# EUROPEAN PATENT SPECIFICATION

(11) **EP 4 573 234 B1**
(45) Date of publication and mention of the grant of the patent: **05.08.2026**
(21) Application number: 23794537.3
(22) Date of filing: 18.08.2023
(51) Int. Cl.: C25B 3/25, C25B 3/26, C25B 9/60, C25B 9/77, C25B 9/75

(54) **MULTI-CELL COX ELECTROLYZER APPARATUS**
MEHRZELLIGE COX-ELEKTROLYSEUR-VORRICHTUNG
APPAREIL D'ÉLECTROLYSE COX MULTICELLULAIRES

(30) Priority: 19.08.2022 US 202263373035 P; 05.06.2023 US 202318329524
(43) Date of publication of application: 25.06.2025
(73) Proprietor: Twelve Benefit Corporation, Berkeley, California 94710 (US); Stone, Simon Gregory, Berkeley, California 94710 (US); Goebel, Steven George, Berkeley, California 94710 (US); Bekkedahl, Timothy A., Berkeley, California 94710 (US); Gallagher, Emerson, Burnaby, British Columbia V5A 4R4 (CA); Moss, Bevan, Burnaby, British Columbia V5A 4R4 (CA); Ma, Sichao, Berkeley, California 94710 (US); Farrell, Noel, Burnaby, British Columbia V5A 4R4 (CA); Whittaker, Dave, Berkeley, California 94710 (US)
(72) Inventor: STONE, Simon Gregory, Berkeley, California 94710 (US); GOEBEL, Steven George, Berkeley, California 94710 (US); BEKKEDAHL, Timothy A., Berkeley, California 94710 (US); GALLAGHER, Emerson, Burnaby, British Columbia V5A 4R4 (CA); MOSS, Bevan, Burnaby, British Columbia V5A 4R4 (CA); MA, Sichao, Berkeley, California 94710 (US); FARRELL, Noel, Burnaby, British Columbia V5A 4R4 (CA); WHITTAKER, Dave, Berkeley, California 94710 (US)
(74) Representative: Optimus Patents Limited
(86) International application number: PCT/US2023/072522
(87) International publication number: WO 2024/040252

(56) References cited:
- JP-A- S5 129 394
- US-A1- 2019 016 616
- US-A1- 2022 243 348

## Description

The present invention relates to a COₓ electrolyzer apparatus, see claim 1.

### BACKGROUND

COₓ electrolyzers offer a potential route for converting or reducing COₓ gas, e.g., CO or CO₂, into one or more desired carbon-based byproducts, such as industrial chemicals or fuels, thereby allowing for waste COₓ gas that would normally be released into the atmosphere to instead be converted into industrially useful products. US2022/243348 describes a COₓ electrolyzer with cathode inlet and outlet ports, Cox electrolyzer cells, a cathode flow field, a Membrane electrode assembly, a cathode gas diffusion layer arranged to receive a COx input and perform electrochemical reduction to provide a range of outputs. US2019/016616 describes an electrochemical cell for wastewater treatment with increased removal rates of pollutants, with a solid polymer electrolyte membrane and an improved current collection and cell compression system. JP S51 29394 describes and electrolytic cell with a sliding electrode chamber.

Background and contextual descriptions contained herein are provided solely for the purpose of generally presenting the context of the present invention. Much of this presents work of the inventors, and simply because such work is described in the background section or presented as context elsewhere herein does not mean that such work is admitted prior art.

### SUMMARY

Details of one or more implementations of the subject matter described in this specification are set forth in the accompanying drawings and the description below. Other features, aspects, and advantages will become apparent from the description, the drawings, and the claims.

The present invention defines a COₓ electrolyzer apparatus according to claim 1, capable of converting or reducing COₓ gas into one or more desired byproducts.

Further preferred embodiment of the present invention are defined in the dependent claims.

In some embodiments, the first components may further include a cathode gas diffusion layer (GDL) adjacent to the cathode frame and covering the cathode flow field. The cathode GDL and the cathode flow field may be configured to guide a flow of gaseous COₓ across the first opening in a first direction transverse to the axial direction and in a distributed manner with respect to at least a second direction transverse to each of the axial and first directions. The second components may further include an anode porous transport layer (PTL) adjacent to the anode frame and covering the anode flow field. The anode PTL and the anode flow field may be configured to guide a flow of anolyte across the second opening in a third direction transverse to the axial direction and in a distributed manner with respect to at least the second direction.

In some embodiments, the cathode frame may include the first opening arranged in a central portion of the cathode frame, at least one first fluidic inlet passage fluidically connected to the anodic parts of the cells, at least one first fluidic outlet passage fluidically connected to the anodic parts of the cells, at least one second fluidic inlet passage fluidically connected to the first opening, and at least one second fluidic outlet passage fluidically connected to the first opening.

### BRIEF DESCRIPTION OF THE DRAWINGS

Various embodiments disclosed herein are illustrated by way of example, and not by way of limitation, in the figures of the accompanying drawings, in which like reference numerals refer to similar elements.
FIG. 1 depicts a diagram of an example MEA for use in COₓ reduction.
FIG. 2 depicts a CO₂ electrolyzer configured to receive water and CO₂ as a reactant at a cathode and expel CO as a byproduct.
FIG. 3 depicts an example construction of a CO₂ reduction MEA having a cathode catalyst layer, an anode catalyst layer, and an anion-conducting PEM.
FIG. 4 depicts an example construction of a CO reduction MEA having a cathode catalyst layer, an anode catalyst layer, and an anion-conducting PEM.
FIG. 5 depicts an exploded view of an example multi-cell COₓ electrolyzer stack.
FIG. 6 depicts a perspective view of the example multi-cell COₓ electrolyzer of FIG. 5.
FIGS. 7 and 8 depict side views of the example multi-cell COₓ electrolyzer of FIG. 6.
FIG. 9 depicts a cross-sectional view of the example multi-cell COₓ electrolyzer of FIG. 7 taken along sectional line 9-9.
FIG. 10 depicts a cross-sectional view of the example multi-cell COₓ electrolyzer of FIG. 8 taken along sectional line 10-10.
FIG. 11A depicts an exploded view of an example repeat unit of the example multi-cell COₓ electrolyzer stack of FIG. 6.
FIG. 11B depicts an exploded view of some cathode components of another example repeat unit of the example multi-cell COₓ electrolyzer stack of FIG. 6.
FIG. 11C depicts a cross-sectional view of the cathode components of the example repeat unit of FIG. 11B.
FIG. 11D depicts an exploded view of anode components of the example repeat unit of the example multi-cell COₓ electrolyzer stack of FIG. 6.
FIG. 11E depicts a cross-sectional view of the anode components of the example repeat unit of FIG. 11D.
FIG. 12 depicts a plan view of an example manifold block of the example multi-cell COₓ electrolyzer of FIG. 6.
FIGS. 13, 14, 15, and 16 depict side views of the example manifold block of FIG. 12.
FIG. 17 depicts an exploded view of an example cathode interface assembly of the example multi-cell COₓ electrolyzer stack of FIG. 6.
FIG. 18 depicts the example cathode interface assembly of FIG. 17 in a non-exploded state.
FIG. 19 depicts an exploded view of an illustrative COₓ electrolyzer cell of the example multi-cell COₓ electrolyzer stack of FIG. 6.
FIG. 20 depicts a bottom view of a representative repeat unit of the example multi-cell COₓ electrolyzer stack of FIG. 6.
FIG. 21 depicts a cross-sectional view of the representative repeat unit of FIG. 20 taken along sectional line 21-21.
FIG. 22 depicts a cross-sectional view of the representative repeat unit of FIG. 20 taken along sectional line 22-22.
FIGS. 23 and 24 depict enlarged portions of the cross-sectional view of FIG. 22.
FIG. 25 depicts a perspective view of the example unitized MEA assembly of the example multi-cell COₓ electrolyzer stack of FIG. 6.
FIG. 26 depicts a top view of the example unitized MEA assembly of FIG. 25.
FIG. 27 depicts a cross-sectional view of the example unitized MEA assembly of FIG. 26 taken along sectional line 27-27.
FIG. 28 depicts a first perspective view of an example cathode frame.
FIG. 29 depicts a bottom view of the example cathode frame of FIG. 28.
FIGS. 30 and 31 depict enlarged portions of the example cathode frame of FIG. 28.
FIG. 32 depicts a second perspective view of the example cathode frame of FIG. 28.
FIG. 33 depicts a top view of the example cathode frame of FIG. 32.
FIG. 34 depicts a cross-sectional view of the example cathode frame of FIG. 33 taken along sectional line 34-34.
FIG. 35 depicts an enlarged portion of the example cathode frame of FIG. 33.
FIG. 36 depicts a cross-sectional view of the example cathode frame of FIG. 35 taken along sectional line 36-36.
FIG. 37 depicts a first perspective view of an example anode frame.
FIG. 38 depicts a top view of the example cathode frame of FIG. 37.
FIG. 39 depicts a second perspective view of the example anode frame of FIG. 37.
FIG. 40 depicts a bottom view of the example anode frame of FIG. 39.
FIG. 41 depicts an enlarged portion of the example anode frame of FIG. 38.
FIG. 42 depicts an enlarged portion of the example anode frame of FIG. 40
FIG. 43 depicts a plan view of an example separator plate of the representative repeat unit of FIG. 11A.
FIG. 44 depicts an example anode interface separator of FIG. 47.
FIGS. 45 and 46 depict top and bottom plan views of an example cathode interface separator of the example cathode interface assembly of FIG. 18.
FIG. 47 depicts an exploded view of an example anode interface assembly of the example multi-cell COₓ electrolyzer stack of FIG. 6.
FIG. 48 depicts the example anode interface assembly of FIG. 47 in an assembled state.
FIG. 49 depicts an example of a cathode flow field with a single serpentine channel.
FIG. 50 depicts a diagram of an example multiple serpentine channel arrangement.
FIG. 51 depicts a diagram of another example multiple serpentine channel arrangement.
FIG. 52 depicts an example of a cathode flow field that includes a two-channel multiple serpentine channel arrangement.
FIGS. 53, 54, and 55 depict an example cathode flow field that may be used in some implementations.
FIGS. 56, 57, and 58 depict an example cathode flow field that may be used in some implementations.
FIG. 59 depicts an example of a cathode flow field that has four cathode serpentine channels arranged in a multiple serpentine channel arrangement.
FIG. 60 depicts a cross-sectional view of a cathode flow field with square- or rectangular-cross-section serpentine channels.
FIG. 61 shows a cross-sectional view of a cathode flow field with a plurality of square- or rectangular-cross-section serpentine channels with rounded interior bottom edges.
FIG. 62 shows a cross-sectional view of a cathode flow field with a plurality of U-shaped cross-section serpentine channels.
FIG. 63 depicts an example of a cathode flow field with peninsular walls having variable wall thickness.
FIG. 64 depicts a plan view of a simplified representation of an example cathode flow field.
FIG. 65 depicts a cathode flow field with two zones and a boundary.
FIG. 66 depicts a cathode flow field with serpentine channels arranged in a bilaterally symmetric manner.
FIG. 67 depicts the same cathode flow field as in FIG. 66 in a scaled-up, broken view manner to allow various features to be more easily labeled and seen.
FIG. 68 depicts another cathode flow field with serpentine channels arranged in a bilaterally symmetric manner.
FIG. 69 depicts the same cathode flow field as in FIG. 68 in a scaled-up, broken view manner to allow various features to be more easily labeled and seen.
FIG. 70 depicts an example of a cathode flow field with a parallel channel arrangement.
FIG. 71 depicts a schematic of an example parallel channel flow field.
FIG. 72 depicts an example of a branching parallel channel flow field.
FIG. 73 depicts the same branching channel flow field as in FIG. 72 but in enlarged form and with the middles of the parallel channels omitted by way of a break section.
FIG. 74 depicts a schematic of another example of a branching parallel channel flow field.
FIG. 75 depicts a schematic of yet another example of a branching parallel channel flow field.
FIG. 76 depicts an example of a cathode flow field that features branching parallel channels.
FIG. 77 depicts a detail view of the left and right sides of the upper half of the cathode flow field of FIG. 76, with the remainder of the flow field omitted from view.
FIG. 78 depicts an example of a cathode flow field with an interdigitated channel arrangement.
FIG. 79 depicts a side view of a gas diffusion layer.
FIG. 80 depicts a flowchart of an example process to form a pre-compressed stack of gas diffusion layers.
FIG. 81 depicts a partial cross-sectional view of an example apparatus to form a pre-compressed stack of gas diffusion layers.
FIG. 82 depicts a partial cross-sectional view of an example roll-to-roll system to form a pre-compressed stack of gas diffusion layers.
FIG. 83 depicts a plan view of a portion of an illustrative anode flow field of the example multi-cell COₓ electrolyzer of FIG. 6.
FIGS. 84A and 84B depict respective cross-sectional views of the illustrative anode flow field of FIG. 83 taken along sectional lines 84A-84A and 84B-84B according to some embodiments.
FIG. 85A depicts a plan view of a portion of an illustrative anode flow field of the example multi-cell COₓ electrolyzer of FIG. 6.
FIGS. 85B and 85C depict respective cross-sectional views of the illustrative anode flow field of FIG. 85A taken along sectional lines 85B-85B and 85C-85C according to some embodiments.
FIG. 86 depicts a plan view of an illustrative insulation plate of the example multi-cell COₓ electrolyzer of FIG. 6.
FIG. 87 depicts a cross-sectional view of the illustrative insulation plate of FIG. 86 taken along sectional line 87-87.
FIG. 88 depicts a plan view of an illustrative end plate of the example multi-cell COₓ electrolyzer of FIG. 6.
FIG. 89 depicts a cross-sectional view of the illustrative end plate of FIG. 88 taken along sectional line 89-89.
FIG. 90 depicts an enlarged portion of the cross-sectional view of FIG. 9
FIG. 91 depicts a perspective view of an example multi-cell COₓ electrolyzer stack.
FIGS. 92 and 93 depict respective side views of the example multi-cell COₓ electrolyzer stack of FIG. 91.
FIGS. 94 and 95 depict respective cross-sectional views the example multi-cell COₓ electrolyzer stack of FIG. 91 respectively taken along sectional lines 94-94 and 95-95.
FIG. 96 depicts a perspective view of an example port side assembly of the example multi-cell COₓ electrolyzer stack of FIG. 91.
FIGS. 97 and 98 depict top and bottom plan views of an example manifold block of the example port side assembly of FIG. 96.
FIGS. 99 and 100 depict bottom and top plan views of an example insulation plate of the example port side assembly of FIG. 96.
FIG. 101 depicts a perspective view of an example piston side assembly of the example multi-cell COₓ electrolyzer stack of FIG. 91 in an exploded state.
FIG. 102 depicts a top plan view of the example piston side assembly of FIG. 101 in an assembled state.
FIG. 103 depicts a cross-sectional view of the example piston side assembly of FIG. 102 taken along sectional line 103-103.
FIG. 104 depicts a perspective view of an example end plate of the example piston side assembly of FIG. 101.
FIGS. 105 and 106 depict a top and bottom plan views of the example end plate of FIG. 104.
FIG. 107 depicts a perspective view of an example piston of the piston side assembly of FIG. 101.
FIGS. 108 and 109 depict top and bottom plan views of the example piston of FIG. 107.

### DETAILED DESCRIPTION OF SOME EMBODIMENTS

COₓ electrolyzers, e.g., CO₂ electrolyzers, using membrane electrode assemblies may share some structural similarities with existing polymer electrolyte membrane (PEM) water electrolyzers, although there are several respects in which COₓ electrolyzers may differ significantly from such PEM water electrolyzer systems.

In a typical COₓ electrolyzer, a membrane electrode assembly (MEA) may be one of multiple elements that are stacked together in what may be referred to as a "cell"; in the discussion below, the term "cell" is used to refer to this multi-element assembly.

An example MEA 100 for use in COₓ reduction is shown in FIG. 1. The MEA 100 has a cathode layer 120 and an anode layer 140 separated by an ion-conducting polymer layer 160 that provides a path for ions to travel between the cathode layer 120 and the anode layer 140. In certain embodiments, the cathode layer 120 includes an anion-conducting polymer and/or the anode layer 140 includes a cation-conducting polymer. In certain embodiments, the cathode layer 120 and/or the anode layer 140 of the MEA 100 are porous. The pores may facilitate gas and/or fluid transport and may increase the amount of catalyst surface area that is available for reaction.

The ion-conducting layer 160 may, for example, include two or three sublayers: a polymer electrolyte membrane (PEM) 165, an optional cathode buffer layer 125, and/or an optional anode buffer layer 145. One or more layers in the ion-conducting layer 160 may be porous. In certain embodiments, at least one layer is nonporous so that reactants and products of the cathode cannot pass via gas and/or liquid transport to the anode and vice versa. In certain embodiments, the PEM layer 165 is nonporous. Example characteristics of anode buffer layers and cathode buffer layers are provided elsewhere herein. In some cases, the ion-conducting layer 160 includes only a single layer or two sublayers.

FIG. 2 shows CO₂ electrolyzer 203 configured to receive water (H₂0) and CO₂ (e.g., humidified or dry gaseous CO₂) as a reactant at a cathode 205 and expel CO as a product. Electrolyzer 203 is also configured to receive water as a reactant at an anode 207 and expel gaseous oxygen (O₂). Electrolyzer 203 includes bipolar layers having an anion-conducting polymer 209 adjacent to cathode 205 and a cation-conducting polymer 211 (illustrated as a proton-exchange membrane) adjacent to anode 207.

As illustrated in the magnification inset of a bipolar interface 213 in electrolyzer 203, the cathode 205 includes an anion exchange polymer (which, in this example, is the same anion-conducting polymer 209 that is in the bipolar layers), electronically conducting carbon support particles 217, and metal nanoparticles 219 supported on the support particles. CO₂ and water are transported via pores (such as pore 221) and reach metal nanoparticles 219 where they react, in this case with hydroxide (OH⁻) ions, to produce bicarbonate (HCO₃) ions and reduction reaction products (not shown). CO₂ may also reach metal nanoparticles 219 by transport within anion exchange polymer 209.

Hydrogen ions are transported from anode 207, and through the cation-conducting polymer 211, until they reach bipolar interface 213, where they are hindered from further transport toward the cathode 205 by anion exchange polymer 209. At interface 213, the hydrogen ions may react with bicarbonate or carbonate ions to produce carbonic acid (H₂CO₃), which may decompose to produce CO₂ and water. As explained herein, the resulting CO₂ may be provided in gas phase and may be provided with a route in the MEA back to the cathode 205 where it can be reduced. The cation-conducting polymer 211 hinders transport of anions, such as bicarbonate ions, to the anode 207 where they could react with protons and release CO₂, which would be unavailable to participate in a reduction reaction at the cathode 205.

As illustrated, a cathode buffer layer having an anion-conducting polymer may work in concert with the cathode 205 and its anion-conductive polymer to block transport of protons to the cathode 205. While MEAs employing ion conducting polymers of appropriate conductivity types in the cathode 205 and cathode buffer layer may hinder transport of cations to the cathode 205 and, if present, an anode buffer layer may similarly hinder transport of the anions to the anode 207, cations and anions may still come in contact in the MEA's interior regions, such as in the membrane layer.

As illustrated in FIG. 2, bicarbonate and/or carbonate ions combine with hydrogen ions between the cathode layer and the anode layer to form carbonic acid, which may decompose to form gaseous CO₂. It has been observed that MEAs sometimes delaminate, possibly due to this production of gaseous CO₂, which does not have an easy egress path.

The delamination issue can be addressed by employing a cathode buffer layer having inert filler and associated pores. One possible explanation of its effectiveness is that the pores create paths for the gaseous carbon dioxide to escape back to the cathode 205 where it can be reduced. In some embodiments, the cathode buffer layer is porous, but at least one layer between the cathode layer and the anode layer is nonporous. This can prevent the passage of gases and/or bulk liquid between the cathode and anode layers while preventing delamination. For example, the nonporous layer can prevent the direct passage of water from the anode 207 to the cathode 205. The porosity of various layers in an MEA is described further at other locations herein.

### Examples of Bipolar MEAs

As an example, an MEA includes a cathode layer including a reduction catalyst and a first anion-conducting polymer (e.g., Sustainion, FumaSep FAA-3, or Tokuyama anion exchange polymer), an anode layer including an oxidation catalyst and a first cation-conducting polymer (e.g., PFSA polymer), a membrane layer including a second cation-conducting polymer and arranged between the cathode layer and the anode layer to conductively connect the cathode layer and the anode layer, and a cathode buffer layer including a second anion-conducting polymer (e.g., Sustainion, FumaSep FAA-3, or Tokuyama anion exchange polymer) and arranged between the cathode layer and the membrane layer to conductively connect the cathode layer and the membrane layer. In this example, the cathode buffer layer can have a porosity between about 1 and 90 percent by volume but can additionally or alternatively have any suitable porosity (including, e.g., no porosity). In other examples the cathode buffer layer can have any suitable porosity (e.g., between 0.01-95%, 0.1-95%, 0.01-75%, 1-95%, 1-90%, etc.).

Too much porosity can lower the ionic conductivity of the buffer layer. In some embodiments, the porosity is 20% or below, and in particular embodiments, between 0.1-20%, 1-10%, or 5-10%. Porosity in these ranges can be sufficient to allow movement of water and/or CO₂ without losing ionic conductivity. Porosity may be measured as described further below.

In a related example, the membrane electrode assembly can include an anode buffer layer that includes a third cation-conducting polymer, and is arranged between the membrane layer and the anode layer to conductively connect the membrane layer and the anode layer. The anode buffer layer preferably has a porosity between about 1 and 90 percent by volume, but can additionally or alternatively have any suitable porosity (including, e.g., no porosity). However, in other arrangements and examples, the anode buffer layer can have any suitable porosity (e.g., between 0.01-95%, 0.1-95%, 0.01-75%, 1-95%, 1-90%). As with the cathode buffer layer, in some embodiments, the porosity is 20% or below, e.g. 0.1-20%, 1-10%, or 5-10%.

In an example, an anode buffer layer may be used in an MEA having a cathode catalyst layer with anion exchange polymer, a cathode buffer layer with anion-exchange polymer, a membrane with cation-exchange polymer, and an anode buffer layer with anion-exchange polymer. In such a structure, the anode buffer layer may be porous to facilitate water transport to the membrane / anode buffer layer interface. Water will be split at this interface to make protons that travel through the membrane and hydroxide that travels to the anode catalyst layer. In some cases, at least one catalyst (e.g., a carbon catalyst, a metal catalyst, etc.) may be utilized to promote the splitting of the water at this interface. For instance, the at least one catalyst may include a cobalt-based catalyst, an iron-nickel-based catalyst, a palladium-based catalyst, platinum-based catalyst, ruthenium (IV) dioxide (RuO₂), nickel-stabilized, ruthenium dioxide (Ni-RuO₂), iridium (IV) dioxide (IrO₂), graphene, graphene oxide (GO), reduced graphene oxide (rGO), graphitic carbon nitride (g-C₃N₄), graphene quantum dots (GQDs), graphene quantum sheets (GQSs), and/or the like. One advantage of this structure is the potential use of low-cost water oxidation catalysts (e.g., NiFeOₓ) that are only stable in basic conditions.

In another specific example, the membrane electrode assembly includes a cathode layer including a reduction catalyst and a first anion-conducting polymer (e.g., Sustainion, FumaSep FAA-3, Tokuyama anion exchange polymer), an anode layer including an oxidation catalyst and a first cation-conducting polymer, a membrane layer including a second anion-conducting polymer (e.g., Sustainion, FumaSep FAA-3, Tokuyama anion exchange polymer) and arranged between the cathode layer and the anode layer to conductively connect the cathode layer and the anode layer, and an anode buffer layer including a second cation-conducting polymer and arranged between the anode layer and the membrane layer to conductively connect the anode layer and the membrane layer.

An MEA containing an anion-exchange polymer membrane and an anode buffer layer containing cation-exchange polymer may be used for CO reduction. In this case, water would form at the membrane / anode buffer layer interface. Pores in the anode buffer layer could facilitate water removal. One advantage of this structure would be the use of an acid-stable (e.g., IrOₓ) water oxidation catalyst.

In a related example, the membrane electrode assembly can include a cathode buffer layer that includes a third anion-conducting polymer and is arranged between the cathode layer and the membrane layer to conductively connect the cathode layer and the membrane layer. The third anion-conducting polymer can be the same or different from the first and/or second anion-conducting polymer. The cathode buffer layer preferably has a porosity between about 1 and 90 percent by volume but can additionally or alternatively have any suitable porosity (including, e.g., no porosity). However, in other arrangements and examples, the cathode buffer layer can have any suitable porosity (e.g., between 0.01-95%, 0.1-95%, 0.01-75%, 1-95%, 1-90%). In some embodiments, the porosity is 20% or below, and in particular embodiments, between 0.1-20%, 1-10%, or 5-10%.

In an example, a cathode catalyst layer composed of Au nanoparticles 4nm in diameter supported on Vulcan XC72 or XC72R carbon and mixed with TM1 (mTPN-1) anion exchange polymer electrolyte may be used. The cathode catalyst layer may be about 15µm thick, have a gold to gold + carbon ratio by weight (Au/(Au+C)) of 20%, have a TM1 to catalyst mass ratio of 0.32, have mass loading of 1.4-1.6 mg/cm² (total Au+C), and have estimated porosity of 0.56. In another example, an anion-exchange polymer layer composed of TM1 and PTFE particles may be provided. The PTFE particles may be approximately 200 nm in diameter and the TM1 molecular weight may be approximately 30k-45k. The thickness of such an example anion-exchange polymer layer may be about 15 µm, and the PTFE particles may introduce a porosity of about 8%. A proton-exchange membrane layer composed of perfluorosulfonic acid polymer (e.g., N afion 115 or Nafion 117) may also be provided, with a thickness of approximately 100 µm to approximately 200 µm. The proton-exchange membrane may form a continuous layer that prevents significant movement of gas (CO₂, CO, H₂) through the layer. An anode catalyst layer composed of Ir or IrOₓ nanoparticles (100-200 nm aggregates) that is 10 µm thick may also be provided.COₓ

### Anion Exchange Membrane-Only MEA for COₓ Reduction

In some embodiments, an MEA does not contain a cation-conducting polymer layer. In such embodiments, the electrolyte is not a cation-conducting polymer and the anode, if it includes an ion-conducting polymer, does not contain a cation-conducting polymer. Various examples thereof are provided below.

An AEM-only MEA allows conduction of anions across the MEA. In embodiments in which none of the MEA layers has significant conductivity for cations, hydrogen ions have limited mobility in the MEA. In some implementations, an AEM-only membrane provides a neutral or an alkaline pH environment (e.g., at least about pH 7) and may facilitate CO₂ and/or CO reduction by suppressing the hydrogen evolution parasitic reaction at the cathode. As with other MEA designs, the AEM-only MEA allows ions, notably anions such as hydroxide, bicarbonate, or carbonate ions, to move through polymer-electrolyte. The pH may be lower in some embodiments; a pH of 4 or greater may be sufficient to suppress hydrogen evolution. The AEM-only MEA also permits electrons to move to, and through, metal and carbon in catalyst layers. In embodiments, the AEM-only MEA may include pores in the anode layer, pores in the cathode layer, and/or pores in the PEM, thereby permiting liquids and gas to move through such pores.

In certain embodiments, the AEM-only MEA comprises an anion-exchange polymer electrolyte membrane positioned between a cathode and an anode. The cathode and the anode are each electrocatalyst layers. In some embodiments, one or both electrocatalyst layers also contain anion-exchange polymer-electrolyte.

In certain embodiments, an AEM-only MEA is formed by depositing cathode and anode electrocatalyst layers onto porous conductive supports, such as gas diffusion layers, porous transport layers, and/or the like, to form gas diffusion electrodes (GDEs). An anion-exchange membrane is then sandwiched between the gas diffusion electrodes.

In certain embodiments, an AEM-only MEA is used for CO₂ reduction. The use of an anion-exchange polymer electrolyte avoids a low pH environment that disfavors CO₂ reduction. Further, water is transported away from the cathode catalyst layer when an AEM is used, thereby preventing water build up (flooding) which can block reactant gas transport in the cathode of the cell.

Water transport in the MEA occurs through a variety of mechanisms, including diffusion and electro-osmotic drag. In some embodiments, at current densities of the CO₂ electrolyzers described herein, electro-osmotic drag is the dominant mechanism. Water is dragged along with ions as they move through the polymer electrolyte. For a cation-exchange membrane such as Nafion membrane, the amount of water transport is well characterized and understood to rely on the pre-treatment/hydration of the membrane. Protons move from positive to negative potential (anode to cathode) with each carrying 2-4 water molecules with it, depending on pretreatment.

In certain embodiments, an AEM-only MEA may be employed in CO reduction reactions. Unlike the CO₂ reduction reaction, CO reduction does not produce carbonate or bicarbonate anions that could transport to the anode and release valuable reactant.

FIG. 3 illustrates an example construction of a CO₂ reduction MEA 301 having a cathode catalyst layer 303, an anode catalyst layer 305, and an anion-conducting PEM 307. In certain embodiments, cathode catalyst layer 303 may include metal catalyst particles (e.g., nanoparticles) that are unsupported or supported on a conductive substrate such as carbon particles. In some implementations, cathode catalyst layer 303 additionally includes an anion-conducting polymer. The metal catalyst particles may catalyze CO₂ reduction, particularly at or within a non-acidic environment. In certain embodiments, anode catalyst layer 305 includes metal oxide catalyst particles (e.g., nanoparticles) that are unsupported or supported on a conductive substrate such as metal oxides, carbides, etc. In some implementations, the anode catalyst layer 305 may additionally include an anion-conducting polymer. Examples of metal oxide catalyst particles for anode catalyst layer 305 may include iridium oxide, nickel oxide, nickel iron oxide, iridium ruthenium oxide, platinum oxide, and the like. The anion-conducting PEM 307 may include any of various anion-conducting polymers such as, for example, HNN5/HNN8 by Ionomr, FumaSep by Fumatech, TM1 by Orion, PAP-TP by W7energy, Sustainion by Dioxide Materials, and the like. These and other anion-conducting polymers that have an ion exchange capacity (IEC) ranging from 1.1 to 2.6, working pH ranges from 0-14, limited solubility in some organic solvents, reasonable thermal stability and mechanical stability, good ionic conductivity/ASR, and acceptable water uptake/swelling ratio may be used. The polymers may be chemically exchanged to certain anions, such as bicarbonate, carbonate, etc., instead of halogen anions prior to use.

As illustrated in FIG. 3, CO₂, such as CO₂ gas, may be provided to cathode catalyst layer 303. In certain embodiments, the CO₂ may be provided via a gas diffusion electrode. At the cathode catalyst layer 303, the CO₂ reacts to produce a reduction product indicated generically as CₓO_{y}H_{z}. Anions produced at the cathode catalyst layer 303 may include hydroxide, carbonate, and/or bicarbonate. These may diffuse, migrate, or otherwise move to the anode catalyst layer 305. At the anode catalyst layer 305, an oxidation reaction may occur such as oxidation of water or hydroxide ion to produce diatomic oxygen and hydrogen ions or water. In some applications, the hydrogen ions may react with hydroxide, carbonate, and/or bicarbonate to produce water, carbonic acid, and/or CO₂. In some cases, fewer interfaces may provide lower resistance for the reaction(s) to occur. In some embodiments, a relatively highly basic environment (e.g., at least a pH above 7) is maintained for C2 and C3 hydrocarbon synthesis.

FIG. 4 illustrates an example construction of a CO reduction MEA 401 having a cathode catalyst layer 403, an anode catalyst layer 405, and an anion-conducting PEM 407. Overall, the constructions of MEA 401 may be similar to that of MEA 301 in FIG. 3. However, the cathode catalyst may be chosen to promote a CO reduction reaction, which means that different reduction catalysts would be used in CO and CO₂ reduction embodiments.

In some embodiments, an AEM-only MEA may be advantageous for CO reduction. The water uptake number of the AEM material can be selected to help regulate moisture at the catalyst interface, thereby improving CO availability to the catalyst. AEM-only membranes can be favorable for CO reduction due to this reason. Bipolar membranes can be more favorable for CO₂ reduction due to better resistance to CO₂ dissolving and crossover in basic anolyte media.

In various embodiments, cathode catalyst layer 403 may include metal catalyst particles (e.g., nanoparticles) that are unsupported or supported on a conductive substrate such as carbon particles. In some implementations, cathode catalyst layer 403 may additionally include an anion-conducting polymer. In certain embodiments, anode catalyst layer 405 includes metal oxide catalyst particles (e.g., nanoparticles) that are unsupported or supported on a conductive substrate such as metal oxides, carbides, etc. In some implementations, the anode catalyst layer 405 may additionally include an anion-conducting polymer. Examples of metal oxide catalyst particles for anode catalyst layer 405 may include those identified for the anode catalyst layer 305 of FIG. 3. Anion-conducting PEM 407 may include any of various anion-conducting polymers such as, for example, those identified for the PEM 307 of FIG. 3.

As illustrated in FIG. 4, CO gas may be provided to cathode catalyst layer 403. In certain embodiments, the CO may be provided via a gas diffusion electrode. At the cathode catalyst layer 403, the CO may react to produce a reduction product indicated generically as CₓO_{y}H_{z}.

Anions produced at the cathode catalyst layer 403 may include hydroxide ions. These may diffuse, migrate, or otherwise move to the anode catalyst layer 405. At the anode catalyst layer 405, an oxidation reaction may occur such as oxidation of water or hydroxide ion to produce diatomic oxygen and hydrogen ions or water. In some applications, the hydrogen ions may react with hydroxide ions to produce water.

While the general configuration of the MEA 401 is similar to that of MEA 301, there are certain differences in the MEAs. For CO₂ reduction, a significant amount of CO₂ may be dissolved and then transferred to the anode for an AEM-only MEA such as shown in FIG. 3. For CO reduction, there is less likely to be significant CO gas crossover. In this case, the reaction environment for CO reduction could be more basic than the reaction environment for CO2 reduction. MEA materials, including the catalyst, may be selected to have good stability in high pH environments.

### Example of AEM-only MEA

1. Copper metal (40 nm thick Cu, about 0.05 mg/cm²) was deposited onto a porous carbon sheet (Sigracet 39BC gas diffusion layer) via electron beam deposition. Ir metal nanoparticles were deposited onto a porous titanium sheet at a loading of 3 mg/cm² via drop casting or ultrasonic spray deposition. An anion-exchange membrane from Ionomr (25-50 µm, 80 mS/cm² OH-conductivity, 2-3 mS/cm² HCO₃⁻ conductivity, 33-37% water uptake) was sandwiched between the porous carbon and titanium sheets with the electrocatalyst layers facing the membrane.

2. Sigma Aldrich 80 nm spherical Cu nanoparticles, mixed with FAA-3 anion exchange solid polymer electrolyte from Fumatech, FAA-3 to catalyst mass ratio of 0.10, setup as described above.

U.S. Patent Application Publication No. US 2017/0321334, published November 9, 2017, and U.S. Patent Application Publication No. 20190226103, published July 25, 2019, which describe various features and examples of MEAs, are incorporated herein by reference in their entireties. All publications referred to herein are incorporated by reference in their entireties as if fully set forth herein.

### Multi-cell COₓ Electrolyzer Stacks

While the above discussion has provided a general overview of various aspects of COₓ MEA construction and characteristics, the following discussion is intended to address aspects of multi-cell COₓ electrolyzer stacks.

FIG. 5 depicts an exploded view of an example multi-cell COₓ electrolyzer stack. FIG. 6 depicts a perspective view of the example multi-cell COₓ electrolyzer of FIG. 5. FIGS. 7 and 8 depict side views of the example multi-cell COₓ electrolyzer of FIG. 6. FIG. 9 depicts a cross-sectional view of the example multi-cell COₓ electrolyzer of FIG. 7 taken along sectional line 9-9. FIG. 10 depicts a cross-sectional view of the example multi-cell COₓ electrolyzer of FIG. 8 taken along sectional line 10-10. FIG. 11A depicts an exploded view of an illustrative repeat unit of the example multi-cell COₓ electrolyzer stack of FIG. 6. FIG. 17 depicts an exploded view of a cathode interface assembly of the example multi-cell COₓ electrolyzer stack of FIG. 6. FIG. 19 depicts an exploded view of an illustrative COₓ electrolyzer cell of the example multi-cell COₓ electrolyzer stack of FIG. 6.

As seen in FIGS. 5-11A, 17, and 19, multi-cell COₓ electrolyzer stack (or stack) 500 includes a plurality of COₓ electrolyzer cells (or cells), such as cell 501, formed by stacking a plurality of repeat units 503 (individually referenced as repeat units 503_1 to 503_n, where "n" is an integer greater than or equal to one) between cathode interface assembly 505 of port side assembly 507 and anode interface assembly 509 of bladder side assembly 511. In this manner, any given cell among the plurality of COₓ electrolyzer cells may be formed by the conjunction of 1) cathode interface assembly 505 (which includes MEA 1105) and anode components 1101 of repeat unit 503_1; 2) cathode components 1103 (which include MEA 1105) of a first repeat unit (e.g., repeat unit 503_1) and anode components 1101 of a second repeat unit (e.g., repeat unit 503_2) adjacent to the first repeat unit; or 3) cathode components 1103 of repeat unit 503_n and anode interface assembly 509. Accordingly, the MEA of any given cell among the plurality of COₓ electrolyzer cells may be configured to facilitate a COₓ reduction process, such as described in association with one or more of FIGS. 1 to 4.

Port side assembly 507 may include cathode interface assembly 505, bus (or terminal) plate 513, manifold assembly 515, insulation plate 517, and end plate 519 sequentially stacked from a first side of the plurality of repeat units 503 in a first direction, e.g., an axial direction, which may extend parallel to the z-axis direction. Among other functions, port side assembly 507 may at least be configured to provide one or more reactants to the cells to feed the COₓ reduction process and output one or more byproducts from the cells in association therewith. Bladder side assembly 511 may include anode interface assembly 509, bus (or terminal) plate 521, insulation plate 523, and end plate 525 sequentially stacked from a second side of the plurality of repeat units 503 in a second direction opposite the first direction. Among other functions, bladder side assembly 511 may be at least configured to constrain axial expansion of the cells during the COₓ reduction process in a manner that prevents or reduces the likelihood of the plurality of cells from being overly compressed, but maintains corresponding fluidic seals and electrical conductivity between associated components of stack 500.

Respective end plates 519 and 525 of port side assembly 507 and bladder side assembly 511 may be coupled to one another via a plurality of tensioning members 527 (e.g., anchors, bolts, studs, tie rods, etc.) extending in the axial direction. As such, end plates 519 and 525 may include respectively pluralities of fastener orifices 519h and 525h through which tensioning members 527 may pass. In some embodiments, fastener orifices 519h and 525h may be respectively arranged about corresponding peripheral regions of end plates 519 and 525. It is also noted that end plates 519 and 525 may be formed of any suitable material, such as aluminum, magnesium, titanium, and/or the like. Tensioning members 527 may be at least partially threaded to respectively engage with, for instance, threaded fasteners 529 (e.g., nuts, rivets, etc.). In this manner, a clamping force extending in the axial direction may be applied to the plurality of cells via the conjunction of end plates 519 and 525, tensioning members 527, and threaded fasteners 529. As such, end plates 519 and 525 may generally serve to act as load-spreading members that distribute a clamping load relatively evenly over the other elements of stack 500. In some instances, first washers 531 may be respectively disposed between the heads of tensioning members 527 and upper surface 519a of end plate 519, and second washers 533 may be respectively disposed between lower surface 525b of end plate 525 and threaded fasteners 529. It is contemplated that one or more of first washers 531 may be formed as lock washers and/or respectively integrated with the heads of tensioning members 527 such as in the case of flanged bolts. Similarly, one or more of second washers 533 may be formed as lock washers and/or respectively integrated with threaded fasteners 529 such as in the case of flanged nuts.

Bus plates 513 and 521 are respectively provided with terminal portions 513t and 521t protruding outwardly from corresponding peripheral surfaces and may be respectively connected to a power supply. In some cases, terminal portions 513t and 521t may have, for example, lugs, terminal blocks, and/or other electrical connection mechanisms to facilitate electrical connections between bus plates 513 and 521 and a corresponding positive or negative voltage or current source. For example, terminal portion 513t on a cathode side of stack 500 may be connected to a negative electrode of the power supply, and terminal portion 521t on an anode side of the stack 500 may be connected to a positive electrode of the power supply. In this manner, bus plates 513 and 521 may provide common electrical connections for the plurality of cells of stack 500, such as cell 501, and, thereby, enable an electrical potential or current to be generated across the plurality of cells of stack 500 that may drive the reduction and oxidation reactions within the plurality of cells. For instance, when an electrical potential difference is imposed on the plurality of cells of stack 500 through application of a voltage or current across bus plates 513 and 521, the resulting electrical potential difference may cause an oxidation reaction at the anode sides of the cells (e.g., oxidation of water to molecular oxygen) and a reduction reaction at the cathode sides of the cells, e.g., that converts the COₓ into carbon monoxide, a hydrocarbon, and/or other catalyst-specific byproducts. As will become more apparent below, bus plate 513 may be sized so as not to interfere with various fluidic passages through stack 500.

According to various embodiments, bus plates 513 and 521 may be formed of a first electrically conductive material, e.g., aluminum, iron, nickel, lead, steel, zinc, and/or the like, and may be coated (or plated) with a second, more electrically conductive coating material, e.g., silver plating, gold plating, copper plating, or other material with relatively higher electrical conductivity, to provide a higher level of electrical conductivity between bus plates 513 and 521 and the corresponding flow fields (e.g., anode and cathode flow fields 1111 and 1127) of the respective cells of stack 500.

Bus plate 513 may, for example, be electrically insulated from end plate 519 by insulation plate 517 and/or at least one other layer of electrically insulating material. As shown, insulation plate 517 is disposed between the electrically conductive portion of bus plate 513 and end plate 519, and may include a plurality of fastener orifices 517h through which tensioning members 527 may pass. In some cases, electrical insulation between bus plate 513 and end plate 519 may be additionally or alternatively provided by manifold assembly 515 when, for instance, manifold assembly 515 is formed of an electrically non-conductive material. Further, electrical insulation may be additionally or alternatively provided by forming (or bonding) electrically insulating material on (or to) a surface of bus plate 513 facing end plate 519, a surface of end plate 519 facing bus plate 513, or at least one surface of manifold assembly 515 facing end plate 519 or end plate 525. Regardless of how such electrical insulation is provided, bus plate 513 may be electrically insulated from end plate 519. When, however, end plate 519 is made of an electrically non-conductive material, or in which end plate 519 is otherwise electrically isolated from, for example, bus plate 521 and/or end plate 525, insulation plate 517 (or other electrically insulating material) may be omitted.

Similar to bus plate 513, bus plate 521 may be electrically insulated from end plate 525 by insulation plate 523 and/or at least one other layer of electrically insulating material that may act in a similar manner as insulation plate 517 with respect to bus plate 513 and end plate 519, but with respect to end plate 525 and bus plate 521. Similar to insulation plate 517, insulation plate 523 may include a plurality of fastener orifices 523h through which tensioning members 527 may pass. In some embodiments, electrical insulation may be additionally or alternatively provided by forming (or bonding) electrically insulating material on (or to) a surface of bus plate 521 facing end plate 525 and/or a surface of end plate 525 facing bus plate 521. In some implementations, insulation plate 523 (or other electrically insulating material) may be omitted if end plate 525 is otherwise electrically isolated from bus plate 521. It is also contemplated that bus plate 521 may be allowed to come into electrically conductive contact with end plate 525 in those instances when the various components of the cells of stack 500 are otherwise configured to maintain electrical insulation between bus plates 513 and 521 other than a conductive path through the various MEAs of the plurality of cells. However, as will become more apparent below, insulation plate 523 may be utilized in association with bus plate 521 to constrain (e.g., actively constrain) axial expansion of the plurality of cells of stack 500. It is noted that an example configuration of insulation plate 523 will be described in more detail in association with FIGS. 86 and 87.

According to some embodiments, insulation plate 523 may be coupled to end plate 525 via a plurality of first fasteners 535. Similarly, insulation plate 517 may be coupled to end plate 519 via a plurality of second fasteners 537. Further, bus plate 513 may be coupled to manifold assembly 515 via a plurality of third fasteners 539. First, second, and third fasteners 535, 537, and 539 may be any suitable fastening mechanism, such as flathead machine screws, rivets, etc., but embodiments are not limited thereto.

### Manifold Assembly

FIG. 12 depicts a bottom plan view of an example manifold block of the example multi-cell COₓ electrolyzer of FIG. 6. FIGS. 13-16 depict side views of the example manifold block of FIG. 12. It is noted that hidden internal features of the manifold block (or main body) 541 that would otherwise not be visible in the view of FIG. 12 are shown in dashed-line format.

In general (and with continued reference to FIGS. 5-10), manifold assembly 515 may be configured to provide one or more reactants to the plurality of cells to feed the COₓ reduction process. For instance, in a COₓ electrolyzer, an anolyte (e.g., liquid water) may be provided to the anode sides of the plurality of cells of stack 500 during operation, while a catholyte (e.g., gaseous COₓ, such as CO and/or CO₂), may be provided to the cathode sides of the cells. In some implementations, an aqueous solution may be provided in place of water, and references to water herein may be understood to also be inclusive of the use of an aqueous solution as well. The liquid water may, through an electrolysis reaction on the anode sides of the cells, undergo oxidation to create oxygen (O₂) gas, H+ protons, and electrons. The H+ protons may be drawn through the MEAs (such as MEA 1105 in FIG. 11A) of the plurality of cells due to an electromagnetic field that is present within the cells due to the electrical potential that is applied across the cells via bus plates 513 and 521 and may react with the bicarbonate and/or hydroxide and/or formate that is produced at the cathode sides of the cells. Manifold assembly 515 may also be configured to allow one or more byproducts of a COₓ reduction process to be expelled from the cells. Thus, as will become more apparent below, manifold assembly 515 may include (or define), for example, at least a portion of one or more fluidic inlet passages and at least a portion of one or more fluidic outlet passages that may be used to convey fluid to and from the anode and cathode sides of the plurality of cells of stack 500.

Referring to FIGS. 5-10 and 12-16, manifold assembly 515 may include main body 541, first fluidic inlet connectors (or couplings) 543, first fluidic outlet connectors 545, second fluidic inlet connector 547, and second fluidic outlet connector 549. Main body 541 may be a generally rectangular plate-shaped body having first surface 1201 opposing second surface 1203 in the axial direction. Although main body 541 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. When assembled as part of stack 500, first surface 1201 may face end plate 525 and interface with bus plate 513 and cathode interface assembly 505, whereas second surface 1203 may face end plate 519 and interface with insulation plate 517. First and second surfaces 1201 and 1203 may be bounded by third, fourth, fifth, and sixth surfaces 1205, 1207, 1209, and 1211. It is noted, however, that embodiments are not limited to the aforementioned configuration, and main body 541 may be formed having any other suitable geometric configuration with corresponding bounding surfaces.

In some embodiments, main body 541 includes first fluidic inlet ports 1213 and 1215 in third and fourth surfaces 1205 and 1207, respectively, that are configured to interface with first fluidic inlet connectors (or inlet connectors) 543, first fluidic outlet ports (or outlet ports) 1217 and 1219 in third and fourth surfaces 1205 and 1207, respectively, that are configured to interface with first fluidic outlet connectors (or outlet connectors) 545, second fluidic inlet port (or inlet port) 1221 in fifth surface 1209 that is configured to interface with second fluidic inlet connector (or inlet connector) 547, and second fluidic outlet port (or outlet port) 1223 in sixth surface 1211 that is configured to interface with second fluidic outlet connector (or outlet connector) 549. As such, first and second inlet and outlet ports 1213-1223 may include corresponding threaded regions, such as threaded region 1215t of first fluidic inlet port 1215 and threaded region 1221t of second fluidic inlet port 1221, to engage with respective threaded regions of first and second fluidic inlet and outlet connectors 543-549. Alternatively, first and second fluidic inlet and outlet connectors 543-549 may be respectively welded, e.g., sweat welded, to first and second inlet and outlet ports 1213-1223 or otherwise coupled to first and second inlet and outlet ports 1213-1223.

First fluidic inlet ports 1213 and 1215 may be fluidically connected to corresponding third fluidic outlet ports in first surface 1201 via respective connecting passages. For instance, first fluidic inlet port 1215 may be fluidically connected to third fluidic outlet port 1225 via connecting passage 1227. Similarly, first fluidic outlet ports 1217 and 1219 may be fluidically connected to corresponding third fluidic inlet ports in first surface 1201 via respective connecting passages. For instance, first fluidic outlet port 1217 may be fluidically connected to third fluidic inlet port 1229 via connecting passage 1231. Third fluidic outlet and inlet ports 1225 and 1229 respectively include a plurality of orifices fluidically connected to one another via corresponding connecting passages. For example, third fluidic outlet port 1225 may include first and second outlet orifices 1225a and 1225b fluidically connected to one another via connecting passage 1233, whereas third fluidic inlet port 1229 may include first and second inlet orifices 1229a and 1229b fluidically connected to one another via connecting passage 1235. Likewise, second fluidic inlet and outlet ports 1221 and 1223 may be fluidically connected to corresponding fourth fluidic outlet and inlet ports 1237 and 1239 in first surface 1201 via respective connecting passages 1241 and 1243. Accordingly, the conjunction of first fluidic inlet ports 1213 and 1215, respective connecting passages (e.g., connecting passage 1227), and corresponding third fluidic outlet ports (e.g., third fluidic outlet port 1225) may be configured to provide water to inlet passages 1001 and 1003 of stack 500. The conjunction of first fluidic outlet ports 1217 and 1219, respective connecting passages (e.g., connecting passage 1235), and corresponding third fluidic inlet ports (e.g., third fluidic inlet port 1229) may be configured to allow water to be expelled from outlet passages of stack 500. It is noted that the outlet passages of stack 500 may be similar to inlet passages 1001 and 1003, but may terminate at first fluidic outlet connectors 545 versus initiate at first fluidic inlet connectors 543. Further, the conjunction of second fluidic inlet port 1221, connecting passage 1241, and fourth fluidic outlet port 1237 may be configured to provide gaseous COₓ to inlet passage 901 of stack 500, whereas the conjunction of second fluidic outlet port 1223, connecting passage 1243, and fourth fluidic inlet port 1239 may be configured to expel one or more byproducts of the COₓ reduction process from outlet passage 903 of stack 500.

In some embodiments, first surface 1201 of main body 541 may include recessed region 1245 configured to receive at least a portion of bus plate 513 therein when manifold assembly 515 is incorporated as part of stack 500. Recessed region 1245 may include one or more portions (e.g., portions 1245a and 1245b) either of which may receive terminal portion 513t of bus plate 513 therein. Additionally, recessed region 1245 may include one or more threaded openings 1247 extending into main body 541 that are configured to threadedly engage with third fasteners (e.g., flatheaded machine screws) 539, which may be utilized to couple bus plate 513 to manifold assembly 515. In some embodiments, threaded openings 1247 may be provided as blind openings including, for instance, swage nuts pressed and/or clinched into main body 541 in a manner that third fasteners 539 engage with the swage nuts. Further, when manifold assembly 515 is incorporated as part of stack 500 and at least a portion of bus plate 513 is received in recessed region 1245, respective fluidic seals may be formed between third fluidic outlet and inlet ports 1225 and 1229 and corresponding ports (or openings) in cathode interface assembly 505 via gaskets 553. Similarly, respective fluidic seals may be formed between fourth fluidic outlet and inlet ports 1237 and 1239 and corresponding ports of cathode interface assembly 505 via gaskets 555.

Main body 541 may further include recesses 1249 and 1251 in third surface 1205 and recess 1253 in fifth surface 1209 to allow datum rods 557 of stack 500 to extend from, for instance, insulation plate 523 in the axial direction and at least partially into corresponding recesses 1249-1253. During assembly of stack 500, datum rods 557 may be utilized to maintain alignment between components of stack 500. In some cases, external surfaces of datum rods 557 may optionally abut against outer surfaces of the plurality of repeat units 503, cathode interface assembly 505, anode interface assembly 509, and/or recesses 1249-1253 of manifold assembly 515.

### Repeat Unit

FIG. 20 depicts a bottom view of a representative repeat unit of the example multi-cell COₓ electrolyzer stack of FIG. 6. FIG. 21 depicts a cross-sectional view of the representative repeat unit of FIG. 20 taken along sectional line 21-21. FIG. 22 depicts a cross-sectional view of the representative repeat unit of FIG. 20 taken along sectional line 22-22. FIGS. 23 and 24 depict enlarged portions of the cross-sectional view of FIG. 22.

Referring to FIGS. 11A and 20-24, representative repeat unit (or repeat unit) 1100 may include separator plate 1107 at least partially stacked between anode components 1101 and cathode components 1103. Anode components 1101 may include anode PTL 1109, anode flow field 1111, first anode gasket set 1113, anode frame 1115, and second anode gasket set 1117. In some embodiments, anode components 1101 may further include anode annular insert 1118 (see FIGS. 11B and 11C). It is noted that various anode components, such as first and second anode gasket sets 1113 and 1117 are not shown in FIGS. 11B and 11C for illustrative convenience. Cathode components 1103 may not only include MEA unit 1119 having MEA 1105 and cathode GDL 1121 stacked between first and second support frames 1123 and 1125, but may also include cathode flow field 1127, first cathode gasket 1129, cathode frame 1131, and second cathode gasket 1133. In some embodiments, cathode components 1103 may further include cathode annular insert 1134 (see FIGS. 11D and 11E). It is noted that various cathode components, such as MEA 1105, first and second support frames 1123 and 1125, and first and second cathode gasket sets 1129 and 1133 are not shown in FIGS. 11B and 11C for illustrative convenience.

According to various embodiments, anode frame 1115 may be coupled to cathode frame 1131 via any suitable fastening mechanism(s), e.g., anchors, bolts, nuts, rivets, screws, and/or the like. For instance, anode frame 1115 may be coupled to cathode frame 1131 via swage (or press) nuts 1135 pressed and/or clinched into anode frame 1115 and fasteners 1137 (e.g., shoulder screws), which interface with cathode frame 1131 and extend through separator plate 1107 to engage with swage nuts 1135. In some embodiments, swage nuts 1135 may be pressed and/or clinched into cathode frame 1131 versus anode frame 1115 such that fasteners 1137 interface with anode frame 1115 and extend through separator plate 1107 to engage swage nuts 1135 of cathode frame 1131. It is also contemplated that a first some of swage nuts 1135 may be pressed and/or clinched into anode frame 1115 and a second some of swage nuts 1135 may be pressed and/or clinched into cathode frame 1131 such that a corresponding first some of fasteners 1137 interface with cathode frame 1131 and extend through separator plate 1107 to engage with the first some of swage nuts 1135 and a corresponding second some of fasteners 1137 interface with anode frame 1115 and extend through separator plate 1107 to engage the second some of swage nuts 1135 of cathode frame 1131. Hereinafter, it will be assumed that swage nuts 1135 are incorporated as part of anode frame 1115 and fasteners 1137 interface with cathode frame 1131 and extend through separator plate 1107 to engage swage nuts 1135 of anode frame 1115. In this manner, second anode gasket set 1117 may be interposed between anode frame 1115 and separator plate 1107, whereas second cathode gasket 1133 may be interposed between separator plate 1107 and cathode frame 1131.

As can be seen in FIGS. 20-24, at least a portion of anode PTL 1109 and anode flow field 1111 may be supported in one or more openings in anode frame 1115, whereas cathode flow field 1127 and at least a portion of unitized MEA assembly 1119 may be supported in one or more openings in cathode frame 1131. In this manner, first cathode gasket 1129 may be interposed between cathode frame 1131 and unitized MEA assembly 1119 to encircle, encompass, circumscribe, surround, and/or the like (hereinafter "encircle") cathode flow field 1127 and bulged portion 1123c (see FIGS. 25-27) of support frame 1123. First anode gasket 1113a of first anode gasket set 1113 may not only be interposed between anode frame 1115 and anode PTL 1109, but may also encircle anode flow field 1111. Second and third anode gaskets 1113b and 1 113c of first anode gasket set 1113 may interface with anode frame 1115 to form fluidic seals with an adjacent repeat unit or cathode interface assembly 505, as will become more apparent below.

According to various embodiments, when repeat unit 1100 is assembled, anode flow field 1111 may be supported in at least one opening in anode frame 1115 such that a first surface of anode flow field 1111 abuts against a corresponding surface of anode PTL 1109 and a second surface of anode flow field 1111 abuts against a corresponding surface of separator plate 1107. In those instances when repeat unit 1100 includes anode annular insert 1118, anode annular insert 1118 may be at least partially supported in at least one opening in anode frame 1115 and may encircle anode flow field 1111. To this end, at least a portion of first surface 1118a (e.g., a top surface) of anode annular insert 1118 may abut against one or more corresponding surfaces of a unitized MEA assembly stacked between two adjacent repeat units or a unitized MEA assembly of cathode interface assembly 505. At least a portion of second surface 1118b (e.g., a bottom surface) of anode annular insert 1118 opposing first surface 1118a may abut against a corresponding surface of anode frame 1115. Additional features and effects of anode annular insert 1118 will be described later in association with anode frame 1115. Similarly, when repeat unit 1100 is assembled, cathode flow field 1127 may be supported in at least one opening in cathode frame 1131 such that a first surface of cathode flow field 1127 abuts against a corresponding surface of separator plate 1107 and a second surface of cathode flow field 1127 at least abuts against a corresponding surface of cathode GDL 1121, which may be exposed by an opening 1123a (see FIGS. 25-27) in support frame 1123 of unitized MEA assembly 1119. In those instances when repeat unit 1100 includes cathode annular insert 1134, cathode annular insert 1134 may be at least partially supported in at least one opening in cathode frame 1131 and may encircle cathode flow field 1127. To this end, at least a portion of first surface 1134a (e.g., a top surface) of cathode annular insert 1134 may abut against a corresponding surface of cathode frame 1131, and at least a portion of second surface 1134b (e.g., a bottom surface) of cathode annular insert 1134 opposing first surface 1134a may abut against one or more corresponding surfaces of a unitized MEA assembly of an associated repeat unit, e.g., repeat unit 1100. Other features and effects of cathode annular insert 1134 will be described later in connection with cathode frame 1131.

Aspects of the various components of repeat unit 1100 will be now described in more detail not only in association with the description of cell 501, but also the text associated with FIGS. 25-43, 49-79, 83, 84A, 84B, and 85A-85C.

### COₓ Electrolyzer Cell

Referring to FIG. 19, an exploded view of cell 501 is shown. Cell 501 is formed between cathode components 1103_1 of repeat unit 503_1 and anode components 1103_2 of repeat unit 503_2. Separator plates 1107_1 and 1107_2 of repeat units 503_1 and 503_2 separate cell 501 from adjacent cells of stack 500. With this in mind, anode components 1101_1 of repeat unit 503_1 and cathode components 1103_2 of repeat unit 503_2 are shown in partially assembled states and form portions of such cells adjacent to cell 501. Hereinafter, components of cell 501 will be referenced followed by an underscore and identifier to indicate the repeat unit to which the components are a part without specifying the repeat unit itself.

Cell 501 may include MEA 1105_1 interposed between anode porous transport layer (PTL) 1109_2 and cathode GDL 1121_1. In some cases, MEA 1105_1 and cathode GDL 1121_1 may be part of a unitized MEA assembly, such as unitized MEA assembly 1119_1, which includes MEA 1105_1 and cathode GDL 1121_1 sandwiched between support frames 1123_1 and 1125_1 (see also FIGS. 25-27). Support frames 1123_1 and 1125_1 may not only include respective openings 1123a_1 and 1125a_1 exposing corresponding surfaces of MEA 1105_1 and cathode GDL 1121_1 to adjacent components, but may also respectively include protruded tab portions 1123b_1 and 1125b_1 that may facilitate handling of unitized MEA assembly 1119_1 during manufacture and testing. In some embodiments, protruded tab portions 1123b_1 and 1125b_1 may be silkscreened, inscribed, embossed, or otherwise marked with identifying information, such as identifying information indicating a cell to which unitized MEA assembly 1119_1 belongs. Support frame 1123_1 may also include bulged portion 1123c_1 (see also bulged portion 1123c in FIG. 27) to accommodate MEA 1105_1 and cathode GDL 1121_1 in a cavity (e.g., cavity 2701 in FIG. 27) formed between support frames 1123_1 and 1125_1. Accordingly, the design of unitized MEA assembly 1119_1 may allow its components to be preassembled and tested before incorporation into, for example, cell 501, which may increase assembly efficiencies and reduce both cell-level and stack-level defects.

With continued reference to FIG. 19, anode PTL 1109_2 may be interposed between MEA 1105_1 and anode flow field 1111_2, whereas cathode GDL 1121_1 may be interposed between MEA 1105_1 and cathode flow field 1127_1. As such, opening 1125a_1 in support frame 1125_1 may allow MEA 1105_1 and anode flow field 1111_2 to be fluidically connected via anode PTL 1111_2, and opening 1123a_1 in support frame 1123_1 may allow MEA 1105_1 and cathode flow field 1127_1 to be fluidically connected via cathode GDL 1127_1. As will become more apparent below, anode PTL 1109_2 and anode flow field 1111_2 may, for example, be supported in one or more openings in anode frame 1115_2 and encircled by first anode gasket 1113a_2 of first anode gasket set 1113_2 at a first side of anode frame 1115_2. Similarly, cathode flow field 1127_1 and at least a portion of unitized MEA assembly 1119_1 (and, thereby, at least cathode GDL 1121_1) may be supported in one or more openings of cathode frame 1131_1 and encircled by first cathode gasket 1129_1 at a first side of cathode frame 1131_1. In turn, anode frame 1115_2 may be stacked between unitized MEA assembly 1119_1 and separator plate 1107_2, and cathode frame 1131_1 may be stacked between separator plate 1107_1 and unitized MEA assembly 1119_1. Second anode gasket set 1117_2 may be disposed between anode frame 1115_2 and separator plate 1107_2, whereas second cathode gasket 1133_1 may be disposed between cathode frame 1131_1 and separator plate 1107_1. In this manner, first anode gasket 1117a_2 of second anode gasket set 1117_2 may encircle anode flow field 1111_2 at a second side of anode frame 1111_2, and second cathode gasket 1133_1 may encircle cathode flow field 1127_1 at a second side of cathode frame 1131_1.

Gaskets 1113a_2 and 1129_1 may not only provide fluidic seals between unitized MEA assembly 1119_1 and the corresponding flow fields 1111_2 and 1127_1, but may also provide structural support to avoid over-compression of anode PTL 1109_2 and cathode GDL 1121_1. It is also noted that gaskets 1113a_2 and 1129_1 may be formed thin enough so that anode PTL 1109_2 and cathode GDL 1121_1 are not under-compressed when assembled as part of stack 500. For example, gaskets 1113a_2 and 1129_1 may be sized such that anode PTL 1109_2 and cathode GDL 1121_1 are compressed and sealed against corresponding surfaces of flow fields 1111_2 and 1127_1 to maintain electrical contact while preventing or discouraging fluids from pooling during operation. In a similar manner, gaskets 1117a_2 and 1133_1 may provide fluidic seals between separator plates 1107_2 and 1107_1 and corresponding surfaces of flow fields 1111_2 and 1127_1.

Each element within cell 501 may provide particular functionality to cell 501, and various components of stack 500 may provide shared functionality with each of the plurality of cells including cell 501. For instance, end plates 519 and 525 may generally serve to act as load-spreading members that distribute a clamping load relatively evenly over the plurality of cells of stack 500 including cell 501. Manifold assembly 515 may include, for example, main body 541 forming at least a portion of one or more fluidic inlet ports, which may begin at inlet connectors 543, and at least a portion of one or more fluidic outlet ports, which may terminate at outlet connectors 545, that may be used to convey fluid to and from the anode sides of the plurality of cells of stack 500 including cell 501. As will become more apparent below, the fluidic inlet port(s) and fluidic outlet port(s) of manifold assembly 515 may be fluidically connected to corresponding inlet and outlet fluidic passages in not only anode frame 1115_2 and cathode frame 1131_1 of cell 501, but also inlet and outlet fluidic passages of the anode and cathode frames of the other cells of stack 500. In a similar fashion, main body 541 of manifold assembly 515 may form at least a portion of one or more fluidic inlet ports, which may begin at inlet connector 547, and at least a portion of one or more fluidic outlet ports, which may terminate at outlet connector 549, that may be used to convey fluid to and from the cathode sides of the plurality of cells of stack 500 including cell 501. Thus, and as will become more apparent below, the fluidic inlet port(s) and fluidic outlet port(s) of manifold assembly 515 may be fluidically connected to corresponding inlet and outlet fluidic passages in not only anode frame 1115_2 and cathode frame 1131_1 of cell 501, but also inlet and outlet fluidic passages of the anode and cathode frames of the other cells of stack 500.

According to various embodiments, bus plate 521 may be electrically connected to anode flow field 1111_2 (and, in some instances, anode frame 1115_2) via anode interface separator 4703, anode flow field 1111, and anode PTL 1109 of anode interface assembly 509 (see FIGS. 5-10 and 47), as well as the corresponding separator plates 1107, anode flow fields 1111, anode PTLs 1109, MEAs 1105, cathode GDLs 1121, and cathode flow fields 1127 between anode interface assembly 509 and cell 501 (see also FIGS. 5-11); similarly, bus plate 513 may be electrically connected to cathode flow field 1127_1 (and, in some instances, cathode frame 1131_1) via cathode interface separator 1701, cathode flow field 1127, cathode GDL 1121, and MEA 1105 of cathode interface assembly 505 (see FIGS. 5-10 and 17). Anode and cathode flow fields 1111_2 and 1127_1 may be made of any suitable material(s) that is electrically conductive and otherwise capable of withstanding relatively long-term exposure to the fluids flowed within stack 500 during normal operating conditions. For example, flow fields 1111_2 and 1127_1 may be made from titanium or titanium alloy, stainless steel (although stainless steel may have a higher susceptibility to corrosion than other materials), porous graphite, a carbon-fiber reinforced thermoset polymer, etc.

In general, anode and cathode frames 1115_2 and 1131_1 may have inlets that correspond in location to the fluidic inlet passageways that begin at inlet connectors 543 and 547, and outlets that corresponding in location to the fluidic outlet passageways that terminate at outlet connectors 545 and 549. To this end, anode and cathode flow fields 1111_2 and 1127_1 may each have one or more channels that are formed in surfaces of the corresponding flow fields that are in contact with anode PTL 1109_2 and cathode GDL 1121_1, respectively, that are routed so as to allow the fluid that is conducted through the channels to come into contact with the adjacent PTL or GDL in a generally distributed manner.

For example, anode flow field 1111_2 may feature one or more inlet openings (or channels) and one or more outlet openings (or channels) that may, respectively, fluidically connect with corresponding openings in anode frame 1115_2. One or more anode channels, e.g., serpentine channels, may be provided in a surface of anode flow field 1111_2 that is in contact with anode PTL 1109_2. The anode channels may serve to distribute the fluid introduced to the anode side of cell 501 across anode PTL 1109_2 such that the anolyte is able to come into contact with anode PTL 1109_2 in a spatially distributed manner such that the anolyte may be allowed to flow through anode PTL 1109_2 in a relatively uniform manner across the entire area, or most of the entire area, of anode PTL 1109_2. An illustrative anode frame 1115 and some example anode flow fields 1111 will be described in more detail in association with FIGS. 37-42 and 83-85.

Similarly, cathode flow field 1127_1 may feature one or more inlet openings (or channels) and one or more outlet openings (or channels) that may, respectively, fluidically connect with corresponding openings in cathode frame 1131_1. One or more cathode channels may be provided in a surface of cathode flow field 1127_1 that is in contact with cathode GDL 1121_1. The cathode channels may serve to distribute the fluid introduced to the cathode side of cell 501 across cathode GDL 1121_1 such that the cathode fluid is able to come into contact with cathode GDL 1121_1 in a spatially distributed manner such that the cathode fluid may be allowed to flow through cathode GDL 1121_1 in a relatively uniform manner across the entire area, or most of the entire area, of cathode GDL 1121_1. An illustrative cathode frame 1131 and example cathode flow fields 1127 will be described in more detail in association with FIGS. 28-36 and 49-78.

Anode PTL 1109_2 and cathode GDL 514 may both serve to help gases that are generated within or provided via anode flow field 1111_2 and cathode flow field 1127_1, respectively, to diffuse across the active area of MEA 1105_1. A typical GDL suitable for use in a COₓ electrolyzer may include, for example, a fibrous substrate that provides structural support, e.g., to the catalyst layer in MEA 1105_1, and may allow gas to flow from the adjacent flow field towards the MEA (including in directions parallel to the plane of MEA 1105_1, thereby allowing the gas to flow laterally underneath portions of the adjacent flow field that may be in contact with the GDL). Such a GDL may also permit water that is present in MEA 1105_1 or that is trapped within the GDL and/or trapped between that GDL and MEA 1105_1 to escape into the channel(s) of a flow field that is adjacent to the GDL, thereby potentially allowing that water to be expelled from that flow field as a result of fluid flow through that flow field. The GDL may also serve as an electrical conductor that serves to conduct electrical charge through MEA 1105_1. Similarly, a typical PTL suitable for use in a COₓ electrolyzer may include, for example, a porous, metallic matrix that provides structural support, e.g., to the catalyst layer in MEA 1105_1, and may allow water to flow from the adjacent flow field towards the MEA (including in directions parallel to the plane of MEA 1105_1, thereby allowing the water to flow laterally above portions of the adjacent flow field that may be in contact with the PTL). Such a PTL may also permit gas that is present in MEA 1105_1 or that is trapped within the PTL and/or trapped between that PTL and MEA 1105_1 to escape into the channel(s) of a flow field that is adjacent to the PTL, thereby potentially allowing that water to be expelled from that flow field as a result of fluid flow through that flow field. The PTL may also serve as an electrical conductor that serves to conduct electrical charge through MEA 1105_1.

According to some embodiments, MEA 1105_1 for a COₓ electrolyzer may feature a metal nanoparticle catalyst layer that is pressed into contact with cathode GDL 1121_1. In some implementations, the metal nanoparticle catalyst layer may alternatively be formed on cathode GDL 1121_1 and pressed into contact with MEA 1105_1. In yet further cases, there may be metal nanoparticle catalyst layers that may be formed on both MEA 1105_1 and cathode GDL 1121_1 and then pressed into contact with each other. One example of such a catalyst layer is a layer of carbon material supporting a layer of, or incorporating, gold nanoparticles. Various types of MEAs and appropriate catalysts for use in a COₓ electrolyzer are discussed in U.S. Patent Application Nos. 15/586,173 and 15/586,182, both filed May 3, 2017, and both titled "REACTOR WITH ADVANCED ARCHITECTURE FOR THE ELECTROCHEMICAL REACTION OF CO2, CO, AND OTHER CHEMICAL COMPOUNDS," and U.S. Patent Application No. 62/939,960, filed November 25, 2019, and titled "MEMBRANE ELECTRODE ASSEMBLY FOR COₓ REDUCTION," each of which is hereby incorporated herein by reference in their entireties. It is noted, however, that these are merely examples and other configurations are contemplated.

Within the context of a multi-cell architecture, such as in the case of stack 500, multiple cells (including cell 501) may be served by common fluidic inlet ports/outlet ports and/or a common electrical potential source. It is noted that the overall multi-cell stack performance may be partially defined by the uniformity of electrical efficiency and product selectivity across the plurality of cells of stack 500, and this uniformity may be driven by the uniformity of gas flow delivery to/across each of the plurality of cells. To this point, the selection of flow field geometry, in that it relates to flow field pressure drop, may have a noticeable effect on overall stack flow uniformity. This may be because the flow uniformity is improved when the pressure drop across/through the plurality of cells is about an order of magnitude more than a pressure difference between discrete locations along a plenum where collective flow is distributed into individual cells within stack 500. Thus, establishing appropriate dimensions may be significant when working with a fixed plenum geometry toward the overall performance of stack 500.

As mentioned earlier, in a COₓ electrolyzer, liquid water may be provided to the anode side of cell 501 during operation, while gaseous COₓ may be provided to the cathode side of cell 501. In some implementations, an aqueous solution may be provided in place of water, and references to water herein may be understood to also be inclusive of the use of an aqueous solution as well. The liquid water may, through an electrolysis reaction on the anode side of cell 501, undergo oxidation to create oxygen (O₂) gas, H+ protons, and electrons. The H+ protons may be drawn through MEA 1105_1 due to the electromagnetic field that is present within cell 501 due to the electrical potential that is applied across cell 501 and may react with the bicarbonate and/or hydroxide and/or formate that is produced at the cathode side.

For a variety of other reasons, water may enter the cathode of MEA 1105_1. In some implementations, liquid water is transported by one or more phenomena to the cathode. Thus, water molecules from the anode side of cell 501 may be transported to the cathode side of cell 501, e.g., through electroosmotic drag caused by the movement of the H+ protons from the anode side of cell 501 to the cathode side of cell 501. The rate of water delivery to and/or generation within the cathode side of cell 501 may be relatively high, e.g., for every molecule of CO gas that is produced through reduction of COₓ gas, there may be, for example, between five (5) and nine (9) molecules of water generated in and/or drawn to the cathode side of cell 501. This imbalance presents a significant challenge-for every molecule of COₓ gas that is reduced on the cathode side of cell 501, between five (5) and nine (9) molecules of water may need to be removed from the cathode side of cell 501. In some COₓ gas electrolyzers, such as those that may use a copper catalyst and may be used to generate CH₄, for every molecule of COₓ gas that is reduced on the cathode side of cell 501, between five (5) and 36 molecules of water may need to be removed from the cathode side of cell 501, presenting an even greater water management challenge.

This imbalance between the rate of COₓ gas reduction and rate of water accumulation on the cathode side of cell 501 is further complicated by the relatively low gas flow rate of COₓ gas as compared with the typical gas flow rate on the cathode side in fuel cells, as well as the relatively lower temperatures and higher pressures used in COₓ electrolyzers as compared with fuel cells. For example, fuel cells may dilute the flow of O₂ in the cathode of a fuel cell using nitrogen (N₂), thereby allowing a higher volumetric flow rate to be used in a fuel cell than may be used in a COₓ electrolyzer. Such higher volumetric flow rates may allow for a faster rate of water molecule evacuation to be provided for in a fuel cell as compared with a COₓ electrolyzer. In contrast, the COₓ gas that is provided to a COₓ electrolyzer may generally be high-purity COₓ gas, which, in combination with the higher working pressures that may be common in COₓ electrolyzers, may allow for much lower volumetric flow rates to be used to provide a similar level of desired reactant gas flow within a COₓ electrolyzer as compared to a comparably sized fuel cell. The generally slower flow rate that is present in a COₓ electrolyzer as opposed to in a fuel cell may, in combination with the higher rate of water creation in and/or migration to the cathode side of cell 501, cause significant issues in a COₓ electrolyzer if not adequately handled that are not as significant a concern in fuel cells.

For example, approximately 90% of the water that is generated in/delivered to the cathode side of the cell during operation of a fuel cell may be in vapor phase, and thus, easily flowed out of the cathode flow field as compared with the water that is generated in/delivered to the cathode side of cell 501 during operation of a COₓ electrolyzer. In a typical COₓ electrolyzer, less than 2% of the gas phase that is generated in/delivered to the cathode side of cell 501 may be water in the vapor phase; the rest is in liquid phase. As a result of this significant liquid/vapor phase imbalance, as well as the significantly higher rate of water condensation in COₓ electrolyzers, COₓ electrolyzers are confronted with unique challenges with liquid water management that are not encountered in fuel cells. Such issues are, of course, also not present in water electrolyzers since the reactant that is delivered to the cathode side of water electrolyzers in the first place is liquid water that migrates from the anode, and the presence of liquid water in the cathode is, thus, not only expected, but desired and by design.

In COₓ electrolyzers, the presence of high concentrations of liquid water on the cathode side of cell 501 presents particular challenges that must be overcome in order for COₓ electrolyzers to be able to operate efficiently. In particular, the presence of liquid water in the cathode side of COₓ electrolyzers may interfere with the flow of gaseous COₓ through cathode GDL 1121_1 to MEA 1105_1 in cell 501. For example, excess liquid water that collects in the cathode channels of cathode flow field 1127_1 and/or cathode GDL 1121_1 may form a physical barrier that occludes portions of the cathode channels of cathode flow field 1127_1 and/or cathode GDL 1121_1 and prevents the gaseous COₓ from coming into contact with some or all of MEA 1105_1. This limits the reduction efficiency of cell 501 and may even, in some cases, cause permanent damage to cell 501 that may decrease the reduction efficiency of cell 501 going forward even if the liquid water is later removed. An additional issue that may occur if there is excess liquid water present in a COₓ electrolyzer is that the water may be reduced instead of the COₓ gas, resulting in the production of hydrogen instead of the desired reaction product.

COₓ electrolyzers may not only experience significantly higher rates of liquid water generation as compared with similarly sized fuel cell reactors, but may also tend to operate under conditions that tend to inhibit, at least in comparison to fuel cells, the ability of COₓ electrolyzers to compensate for such increased liquid water generation in some respects. For example, the input gas, e.g., air, that is provided to the cathode side of fuel cells tends to be provided at a higher flow rate as compared with the input gas that is provided to the cathode side of COₓ electrolyzers. As air is abundantly available, there is little concern with respect to a fuel cell with providing more air than can be utilized in the reduction reaction of a fuel cell. As a result, air may be provided to the cathode flow field in a fuel cell at a much higher flow rate than may be needed in order to support the reduction reaction taking place within the fuel cell, thereby allowing more kinetic energy to be available in fuel cell cathode input gas flows that may be used to assist with forcibly expelling water that has accumulated within the fuel cell cathode flow field. Further, in fuel cells, the oxidant gas may commonly be diluted with other gases, e.g., nitrogen in air, and higher flow rates may, thus, be used to ensure a sufficient rate of delivery of the oxidant gas to the cathode side of the fuel cell. The increased flow velocity in fuel cells may serve to forcibly push any potential droplets of liquid water that are present in the cathode flow field channel(s) through the flow field and to the fluidic outlet port of the cathode flow field, thereby rapidly evacuating what little liquid water is present in the flow field channels from the flow field.

In contrast, the input gas in a COₓ electrolyzer is the COₓ gas, and one of the main reasons for using COₓ electrolyzers is to reduce COₓ emissions that may be harmful to the environment by converting COₓ gas to other, more desirable gases or liquids (e.g., commercially valuable gases or liquids or gases or liquids that are less harmful to the environment, e.g., water and/or oxygen). It may, thus, be desirable to reduce the flow rate of the COₓ gas to a level that still achieves high, and preferably maximal, COₓ reduction for a given electrical current density used with a COₓ electrolyzer, but also reduces or minimizes the amount of extra COₓ gas that is flowed through the COₓ electrolyzer and is not reduced.

Due to such factors, COₓ electrolyzers may operate using a high-purity, undiluted input gas stream or streams, e.g., pure COₓ gas or relatively pure COₓ gas, that is flowed into the cathode side of cell 501 at relatively low speeds, at least as compared with equivalently sized fuel cells having similar construction. For example, some COₓ electrolyzers may be capable of operating at flow speeds comparable to or lower than those found in a typical fuel cell. In some implementations, COₓ electrolyzers are configured to operate at an average COₓ gas flow velocity in the flow field channels of between about 0.02 m/s and about 30 m/s, between about 0.02 m/s and about 15 m/s, between about 15 m/s and about 30 m/s, between about 0.02 m/s and about 7.5 m/s, between about 7.5 m/s and about 15 m/s, between about 15 m/s and about 23 m/s, between about 23 m/s and about 30 m/s, between about 0.02 m/s and about 3.8 m/s, between about 3.8 m/s and about 7.5 m/s, between about 7.5 m/s and about 11 m/s, between about 11 m/s and about 15 m/s, between about 15 m/s and about 19 m/s, between about 19 m/s and about 23 m/s, between about 23 m/s and about 26 m/s, or between about 26 m/s and about 30 m/s. In some implementations, COₓ electrolyzers are configured to operate at a COₓ gas flow velocity of about 2 m/s to 10 m/s, or about 5 m/s to 10 m/s, or about 7.5 m/s to about 10 m/s.

As indicated, in some implementations, relatively low flow rates provide advantages in COₓ electrolyzers, such as relatively high COₓ utilizations (not to be confused with conversion efficiency) due to low molar flow rates, which are often associated with low volumetric or linear flow rates. Another benefit is in maintaining the MEA (e.g., MEA 1105_1 of cell 501) at an acceptable hydration level. High gas flow rates tend to dry out the MEA, which leads to degradation. Further, for a fixed utilization, flow field designs having shorter channels, and hence more channels per cell, allow for lower gas speeds. In some embodiments, COₓ electrolyzers are configured to operate at a COₓ flow speed in flow channels of between about 0.02 m/s and about 5 m/s, between about 0.02 m/s and about 2.5 m/s, between about 2.5 m/s and about 5 m/s, between about 0.02 m/s and about 1.3 m/s, between about 1.3 m/s and about 2.5 m/s, between about 2.5 m/s and about 3.8 m/s, between about 3.8 m/s and about 5 m/s, between about 0.02 m/s and about 0.64 m/s, between about 0.64 m/s and about 1.3 m/s, between about 1.3 m/s and about 1.9 m/s, between about 1.9 m/s and about 2.5 m/s, between about 2.5 m/s and about 3.1 m/s, between about 3.1 m/s and about 3.8 m/s, between about 3.8 m/s and about 4.4 m/s, or between about 4.4 m/s and about 5 m/s.

In contrast, the typically lower flow rates seen in COₓ electrolyzers, coupled with the significantly higher rates of liquid water introduction into the cathode side of cell 501, make water evacuation in COₓ electrolyzers much more challenging as compared with other electrochemical devices, e.g., fuel cells or water electrolyzers.

Accordingly, various features and technologies may be used to help mitigate the detrimental effects of liquid water accumulation in COₓ electrolyzer cathodes, as well as liquid water supply in COₓ electrolyzer anodes. For example, anode frame 1115_2, cathode frame 1131_1, anode flow field 1111_2, and cathode flow field 1127_1 may be constructed so as to have one or more structural features that may allow for more effective liquid water management in cell 501. For example, anode frame 1115_2, cathode frame 1131_1, anode flow field 1111_2, and cathode flow field 1127_1 may have corresponding channels, risers, protrusions, distributors, collectors, etc., that may, for example, be designed to have certain characteristics that may contribute to 1) more effective water and gaseous COₓ delivery to the anode and cathode sides of cell 501, 2) more effective water evacuation in the context of a COₓ electrolyzer, 3) more effective mitigation of the potential performance degradation that may occur in such a COₓ electrolyzer in the event that liquid water collects within, for instance, the cathode side of cell 501, and 4) more effective expulsion from cell 501 of the byproducts of the COₓ reduction process. Accordingly, cathode frame 1131_1, anode frame 1115_2, cathode flow field 1127_1, and anode flow field 1111_2 will now be discussed in more detail in association with FIGS. 28-78, 83, 84A, 84B, and 85A-85C.

### Cathode Frame

As previously discussed in association with FIGS. 5-11A, cathode flow field 1127 may be supported in an opening of cathode frame 1131 between separator plate 1107 and unitized MEA assembly 1119, as well as include a plurality of fluidic passages to facilitate fluid flow (or communication) through stack 500, and, in particular, through a cell of stack 500, such as cell 501. Various details of an illustrative cathode frame 1131 will now be discussed in more detail in association with FIGS. 28-36.

FIG. 28 depicts a first perspective view of an example cathode frame. FIG. 29 depicts a bottom view of the example cathode frame of FIG. 28. FIGS. 30 and 31 depict enlarged portions of the example cathode frame of FIG. 28. FIG. 32 depicts a second perspective view of the example cathode frame of FIG. 28. FIG. 33 depicts a top view of the example cathode frame of FIG. 32. FIG. 34 depicts a cross-sectional view of the example cathode frame of FIG. 33 taken along sectional line 34-34. FIG. 35 depicts an enlarged portion of the example cathode frame of FIG. 33. FIG. 36 depicts a cross-sectional view of the example cathode frame of FIG. 35 taken along sectional line 36-36.

Cathode frame (or frame) 1131 may be a generally rectangular plate-shaped body having first surface 2801 (e.g., a top surface) opposing second surface 2803 (e.g., a bottom surface) in axial direction 2901 (see FIG. 29). Although frame 1131 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, frame 1131 will be described in association with a generally rectangular configuration. First and second surfaces 2801 and 2803 may be bounded by one or more peripheral surfaces, such as peripheral surfaces (or surfaces) 2805, 2807, 2809, and 2811 that may be connected to one another via one or more other peripheral surfaces, such as peripheral surface (or surface) 2813. In some embodiments, frame 1131 may have a symmetrical configuration about one or more reference planes perpendicular to axial direction 2901 shown in FIG. 29. For instance, a configuration of frame 1131 may be symmetrical about either or both of reference planes 2903 and 2905 (see FIG. 29), but embodiments are not limited thereto.

According to various embodiments, first fluidic inlet passages 2815 and 2817 may be adjacent to peripheral edge 2805, and first fluidic outlet passages 2819 and 2821 may be adjacent to peripheral edge 2809. First fluidic inlet passages 2815 and 2817 may form portions of inlet passages 1001 and 1003 (see FIG. 10) of stack 500 in association with inlet connectors 543 of manifold assembly 515 (see FIGS. 5-10) that provide input water to the various anode frames (e.g., anode frame 1115 in FIG. 11A) of stack 500, and, thereby, to the corresponding anode flow fields (such as anode flow field 1111 in FIG. 11A) of the plurality of cells, such as cell 501. First fluidic outlet passages 2819 and 2821 may form portions of outlet passages (that are similar to inlet passages 1001 and 1003 (see FIG. 10), but associated with outlet connectors 545 of manifold assembly 515 versus inlet connectors 543 (see FIG. 5)) of stack 500 that output water from the various anode frames of stack 500, such as anode frame 1115 in FIG. 11A, and, thereby, from corresponding anode flow fields (e.g., anode flow field 1111 in FIG 11) of the plurality of cells. In some cases, first fluidic inlet and outlet passages 2815-2821 may be defined by respective pluralities of orifices separated from one another via corresponding septal walls. For instance, first fluidic inlet passage 2815 may include first and second inlet orifices 2815a and 2815b separated from one another via septal wall 2803s1, whereas first fluidic outlet passage 2819 may include first and second outlet orifices 2819a and 2819b separated from one another via septal wall 2803s2. Illustrative septal walls are also depicted in the cross-sectional views of FIGS. 23 and 34. For example, septal wall 2803s3 is shown separating first and second outlet orifices 2821a and 2821b forming first fluidic outlet passage 2821 in FIG. 34, and septal wall 2803s4 is shown separating first and second inlet orifices 2817a and 2817b forming first fluidic inlet passage 2817 in FIG. 23. The presence of these septal walls, such as septal walls 2803s1-2803s4, may increase the structural rigidity and, thereby, reliability of frame 1131 in the vicinity of first fluidic inlet and outlet passages 2815-2821.

According to various implementations, frame 1131 includes through opening (or opening) 2823 formed completely through a first central portion of frame 1131 and may be configured to receive at least a portion of cathode flow field 1127 (see, e.g., FIGS. 11A, 23, and 24) therein. In this manner, opening 2823 may be shaped and sized to correspond with the shape and size of cathode flow field 1127. For example, opening 2823 may have a generally rectangular shape with rounded corners, but embodiments are not limited thereto. Frame 1131 may also include blind opening (or opening) 2825 formed in a second central portion of frame 1131 encircling the first central portion of frame 1131. In some cases, opening 2825 may be omitted or may be at least partially filled by cathode annular insert 1134, as will become more apparent below. When included as part of cathode frame 1131, opening 2825 may terminate at surface 2803r, which may be recessed from second surface 2803, and may be configured to receive at least a portion of unitized MEA assembly 1119 (see, e.g., FIGS. 11A, 23, and 24) and/or at least a portion of cathode annular insert 1134 therein. As such, opening 2825 may be shaped and sized to correspond with the shape and size of the portion of unitized MEA assembly 1119 and/or cathode annular insert 1134, but embodiments are not limited thereto. For instance, opening 2825 may have a generally rectangular shape with rounded corners, but embodiments are not limited thereto. In some implementations, the sides of opening 2825 extending respectively adjacent to surfaces 2805 and 2809 of frame 1131 may bulge towards surfaces 2805 and 2809, and, thereby, away from opening 2823. For example, as seen in FIGS. 29 and 31, the side of opening 2825 extending adjacent to surface 2809 of frame 1131 may not only have central portion 2825a extending in a first direction parallel (or substantially parallel) to surface 2809, but may also have second portions 2825b extending from central portion 2825a that are angled inwards from first portion 2825a towards opening 2823 by, for instance, angle 3101. Central portion 2825a may have width 3103 in the first direction, whereas second portions 2825b may have corresponding widths 3105, which may be greater than width 3103. Curved (or arcuate) corners 2825c of opening 2825 may respectively extend from second portions 2825b to connect the side of opening 2825 extending adjacent to surface 2809 to corresponding sides of opening 2825 extending in a second direction transverse to the first direction, e.g., extending parallel (or substantially parallel) to surfaces 2807 and 2811 of frame 1131. Embodiments, however, are not limited thereto.

In those implementations including cathode annular insert 1134, cathode annular insert 1134 may be at least partially supported in opening 2825 such that first surface 1134a of cathode annular insert 1134 abuts against surface 2803r of frame 1131 and inner peripheral surface 1134c of cathode annular insert 1134 encircles an outer peripheral boundary of cathode flow field 1127, and thereby, an inner peripheral boundary of opening 2825 (see also FIGS. 11D and 11E). To this end, outer peripheral surface 1134d of cathode annular insert 1134 may be shaped and sized to correspond with the shape and size of an inner peripheral boundary of opening 2825. In some cases, thickness 1134t of cathode annular insert 1134 may be equivalent (or substantially equivalent) to the depth of opening 2825, but implementations are not limited thereto. When thickness 1134t of cathode annular insert 1134 corresponds to the depth of opening 2825, cathode annular insert 1134 may fill the void in cathode frame 1131 corresponding to opening 2825. It is also contemplated that cathode annular insert 1134 may include one or more notched portions 1134n1 and 1134n2 such that cathode annular insert 1134 does not completely fill the void corresponding to opening 2825. Whatever the case, cathode annular insert 1134 may have a generally ring-like configuration, and as such, may not be truly annular. For instance, cathode annular insert 1134 may have a generally rectangular cross-section when viewed along the z-axis direction shown in FIGS. 11D and 11E, thus giving rise to a cathode annular insert having twofold symmetry instead of axial symmetry. As such, cathode annular insert 1134 may have, for instance, a circular, an oval, a polygonal, or any other suitable cross-sectional geometry when viewed along the z-axis direction shown in FIGS. 11D and 11E.

As seen in FIG. 29, openings 2823 and 2825 may be arranged between second fluidic inlet and outlet passages 2827 and 2829, which form respective portions of inlet and outlet passages 901 and 903 of stack 500 in association with input and outlet connectors 547 and 549 of manifold assembly 515 (see FIGS. 5 and 9). Referring momentarily to FIGS. 7, 9, 11A, 23, 24, and 29, inlet passage 901 may supply one or more reactants (e.g., gaseous COₓ) to frame 1131, and, thereby, to cathode flow field 1127 at least partially supported in opening 2823 when frame 1131 is incorporated as part of a cell, such as cell 501. Outlet passage 903, however, may enable one or more byproducts of the COₓ reduction process to be routed from frame 1131, and, thereby, from the corresponding cathode flow field 1127 at least partially supported in one or more of openings 2823 and 2825. Adverting back to FIGS. 28-36, to enable such exchange of fluids to and from cathode flow field 1127 (see FIG. 11A), second fluidic inlet passage 2827 may be fluidically connected to opening 2823 via channel 3501, connecting riser 3001, and buffering passage 2831, and second fluidic outlet passage 2829 may be fluidically connected to opening 2823 via channel 3301, connecting riser 3109, and buffering passage 2833.

Buffering passages 2831 and 2833 may be corresponding recesses formed in surface 2803r that respectively terminate at surfaces 2831a and 2833a. To facilitate reactant supply to, and byproduct expulsion from, the corresponding cathode flow field 1127 (see, e.g., FIGS. 23 and 24) at least partially supported in opening 2823, buffering passages 2831 and 2833 may have corresponding outer sidewalls 2831b and 2833b that respectively expand from connecting risers 3001 and 3109 towards opening 2823. For instance, buffering passages 2831 and 2833 may have a generally triangular shape, but embodiments are not limited thereto. In some instances, respective widths 3111 of buffering passages 2831 and 2833 may be smaller than width 3103 of central portion 2825a of opening 2825. Buffering passages 2831 and 2833 may also include corresponding pluralities of protrusions 3003 arranged at one or more intervals to accelerate reactant/byproduct flow between adjacent protrusions among the protrusions 3003 and between protrusions 3003 and correspondingly adjacent sidewalls 2831b and 2833b. In association with buffering passage 2831, protrusions 3003 may not only promote a draw of reactant from connecting riser 3001, but may also facilitate a distributed flow of reactant to an input portion of cathode flow field 1127 (see, e.g., FIGS. 23 and 24) at least partially supported in opening 2823. Protrusions 3003, in association with buffering passage 2833, may promote a draw of byproduct from an output portion of cathode flow field 1127 (see, e.g., FIGS. 23 and 24) at least partially supported in opening 2823 to connecting riser 3109. Although protrusions 3003 are shown as generally cylindrically shaped bosses, embodiments are not limited thereto. For instance, one or more of protrusions 3003 may be generally elliptical bosses, generally rectangular bosses, generally pentagonal bosses, generally hexagonal bosses, etc. When incorporated as part of a cell, such as cell 501, cathode annular insert 1134 may be at least partially supported in opening 2825 to at least partially fill the void corresponding to opening 2825. By filling the void corresponding to opening 2825 (which is formed between opening 2823 in frame 1131 and recess 2835) the likelihood that input reactant(s) (e.g., gaseous COₓ) that are to be supplied to cathode flow field 1127 from buffering passage 2831 instead flow around cathode flow field 1127 via opening 2825 (illustrated in FIG. 11D as reactant bypass flow 1136) and become expelled via buffering passage 2833 is reduced or eliminated. It is noted that reactant bypass flow 1136 decreases the amount of input reactant flowing through cathode flow field 1134, and as such, has the potential to decrease the efficiency of the cell. In some cases, both opening 2825 and cathode annular insert 1134 may be omitted, thereby further reducing the possibility of reactant bypass flow 1136. In those instances when opening 2825 is formed in frame 1131 and cathode annular insert 1134 is not utilized, the compression of at least a portion of unitized MEA assembly 1119 therein may also serve to reduce or prevent reactant bypass flow 1136.

According to some embodiments, the inclusion of cathode annular insert 1134 may also aid in providing additional compression of GDL 1121 in the region occupied by cathode annular insert 1134 when the cell (e.g., cell 501) and/or stack 500 is assembled and compressed, whether as part of the assembly process or during use of stack 500. This additional compression may decrease in-plane permeability of GDL 1121 in the region corresponding to cathode annular insert 1134 and may further mitigate the potential for reactant bypass flow 1136. Given, however, that the presence of cathode annular insert 1134 between GDL 1121 and frame 1131 is likely to compress cathode annular insert 1134 in the axial direction, notched portions 1134n1 and 1134n2 may be formed in cathode annular insert 1134 in areas corresponding to buffering passages 2831 and 2833 to prevent or reduce the likelihood that cathode annular insert 1134 compresses into respective portions of buffering passages 2831 and 2833 that interface with opening 2823 in frame 1131. As such, notched portions 1134n1 and 1134n2 may be formed such that their leading edges corresponding to portions of inner peripheral surface 1134c of cathode annular insert 1134 overlap with corresponding protrusions 3003 respectively formed in buffering passages 2831 and 2833 to support cathode annular insert 1134 in the areas corresponding to buffering passages 2831 and 2833. For example, the leading edges of notched portions 1134n1 and 1134n2 may be supported by one or more of protrusions 3003. In some examples, the leading edges of notched portions 1134n1 and 1134n2 may be supported by one or more of protrusions 3003 positioned nearest to connecting riser 3001. Notched portions 1134n1 and 1134n2, however, may be omitted. In some cases, additional protrusions 3003 may be provided in buffering passages 2831 and 2833 to support cathode annular insert 1134 thereon, and thereby, to similarly prevent or reduce the likelihood that cathode annular insert 1134 compresses into the respective portions of buffering passages 2831 and 2833 that interface with opening 2823 in frame 1131.

In some embodiments, protrusions 3003 may be sized similar (or substantially similar) to one another or at least one protrusion among protrusions 3003 may be sized differently than at least one other protrusion among protrusions 3003. This may be with respect to the lengths, widths, and/or heights of protrusions 3003. For example, protrusions 3003 may include first, second, and third protrusions 3003a, 3003b, and 3003c. With respect to a reference plane perpendicular to the axial direction, a cross-sectional area of first protrusions 3003a may be larger than a cross-sectional area of second protrusions 3003b, and a cross-sectional area of second protrusions 3003b may be larger than a cross-sectional area of third protrusions 3003c. In some cases, second protrusions 3003b of buffering passages 2831 and 2833 may be disposed respectively closer to connecting risers 3001 and 3109 than first and third protrusions 3003a and 3003c. Third protrusions 3003c may be arranged amongst first protrusions 3003a and positioned such that third protrusions 3003c are disposed between second protrusions 3003b and a majority of first protrusions 3003a. Embodiments, however, are not limited to such a configuration and/or arrangement of protrusions 3003.

Frame 1131 may also include recess 2835 in surface 2803 and recess 3303 in surface 2801 that are configured to respectively receive corresponding portions of first and second cathode gaskets 1129 and 1133 (see, e.g., FIGS. 11A, 23, and 24) therein when, for example, frame 1131 is assembled as part of a repeat unit (e.g., repeat unit 503_1 in FIG. 5) or cathode interface assembly 505 (see FIG. 5). Recess 2835 may be formed to encircle the periphery of opening 2825 and recess 3303 may be formed to encircle the periphery of opening 2823. It is noted that the conjunction of second fluidic inlet passage 2827, channel 3501, connecting riser 3001, and buffering passage 2831 enables reactant supply to flow from an area outside of first cathode gasket 1129 (see, e.g., FIGS. 11A, 23, and 24) to an area inside of first cathode gasket 1129 without disturbing the integrity of or seal provided by first cathode gasket 1129. Similarly, the conjunction of buffering passage 2833, connecting riser 3109, channel 3301, and second fluidic outlet passage 2829 enables byproduct flow from an area inside of first cathode gasket 1129 (see, e.g., FIGS. 11A, 23, and 24) to an area outside of first cathode gasket 1129 without disturbing the integrity of or seal provided by first cathode gasket 1129.

According to some embodiments, frame 1131 may include first protruded portions 3305 extending from surface 2801 and encircling corresponding first fluidic inlet and outlet passages 2815, 2817, 2819, and 2821. Second protruded portions 3307 may also extend from surface 2801, but encircle respective second fluidic inlet and outlet passages 2827 and 2829. In some implementations, the second protruded portion 3307 encircling second fluidic inlet passage 2827 may also encircle channel 3501 and connecting riser 3001, and the second protruded portion 3307 encircling second fluidic outlet passage 2829 may also encircle channel 3301 and connecting riser 3109. In some embodiments, first and second protruded portions 3305 and 3307 may protrude from surface 2801 by height 3401, but embodiments are not limited thereto. For instance, one or more of first and second protruded portions 3305 and 3307 may have a different height than at least another one or more of first and second protruded portions 3305 and 3307. When assembled as part of a repeat unit (e.g., repeat unit 1100 in FIG. 11A), first and second protruded portions 3305 and 3307 of frame 1131 may be received in and through corresponding openings in a separator plate (such as separator plate 1107 in FIG. 11A; see also FIGS. 23 and 24) or corresponding recesses 4607-4617 (see FIG. 46) in cathode interface separator 1701 (see FIG. 17) of cathode interface assembly 505 (see, e.g., FIGS. 5-10 and 17). As such, one or more of first and second protruded portions 3305 and 3307 may be sized to form respective clearance or interference fits with the corresponding openings in the separator plate (such as separator plate 1107 in FIG. 11A) or corresponding recesses 4607-4617 (see FIG. 46) in cathode interface separator 1701 (see FIGS. 17 and 46) when frame 1131 is assembled as part of a repeat unit (e.g., repeat unit 503_1 in FIG. 5 or as part of cathode interface assembly 505, see, e.g., FIGS. 5-10, 17, and 18).

In some embodiments, one or more of first and second protruded portions 3305 and 3307 may be sized to form respective clearance fits with corresponding features in (or of) the separator plate to which frame 1131 interfaces when incorporated as part of stack 500 (such as separator plate 1107 in FIG. 11A) or cathode interface separator 1701 (see, e.g., FIG. 17) depending on the location of frame 1131 within stack 500). In addition, one or more of first and second protruded portions 3305 and 3307 may be sized to form respective interference fits with the corresponding features in the separator plate to which frame 1131 interfaces when incorporated as part of stack 500 (such as separator plate 1107 in FIG. 11A) or cathode interface separator 1701 (see, e.g., FIG. 17) depending on the location of frame 1131 within stack 500). For example, respective outer boundaries of first and second protruded portions 3305 and 3307 may be about 0.01% to about 5% larger (in the case of an interference fit) or about 0.01% to about 10% smaller (in the case of a clearance fit) than corresponding boundaries of the corresponding features in the separator plate (such as separator plate 1107 in FIG. 11A) or cathode interface separator 1701 (see, e.g., FIG. 17) depending on the location of frame 1131 within stack 500). The clearance and/or interference fits may be utilized to constrain in-plane expansion (e.g., expansion in, for instance, a plane parallel to an x-y plane (see FIG. 11A)) of frame 1131 (and, in some embodiments, anode frame 1115) during operation of stack 500 without unduly stressing frame 1131 and/or anode frame 1115. In some embodiments, first and second protruded portions 3305 and 3307 may be sized to form respective clearance fits with corresponding features in (or of) the separator plate (such as separator plate 1107 in FIG. 11A) or cathode interface separator 1701 (see, e.g., FIG. 17) depending on the location of frame 1131 within stack 500) in a cooled, non-operational state of stack 500 (see FIGS. 5 and 6), but expand to form corresponding interference fits in a steady-state operational condition of stack 500. This may prevent (or at least reduce the likelihood of) misalignments, bunching, etc., of cathode GDLs 1121 and anode PTLs 1109 of the various cells of stack 500, as well as prevent (or reduce the likelihood of) misalignments between adjacent frames of adjacent cells of stack 500. Such a configuration may also allow frame 1131 and/or anode frame 1115 (see FIG. 11A) to be formed of more compliant materials that, in some cases, may be less expensive and/or easier to manufacture (and, in some cases, not electrically conductive). It is noted, however, that the separator plate (e.g., separator plate 1107 in FIG. 11A) or cathode interface separator 1701 (see, e.g., FIG. 17) depending on the location of frame 1131 within stack 500) may be formed of a stronger and/or more rigid material(s) to increase the strength and/or rigidity of the various repeat units (e.g., repeat unit 1100 of FIG. 11A; see also repeat units 503 in FIGS. 5-10) and/or cathode interface assembly 505 (see, e.g., FIGS. 5-10, 17, and 18).

According to various embodiments, first protruded portions 3305 may be sized and shaped to interface with second anode gaskets 1117b of second anode gasket set 1117 and second protruded portions 3307 may be sized and shaped to interface with third anode gaskets 1117c of second anode gasket set 1117. As such, cross-flow between first and second fluidic inlet and outlet passages 2815, 2817, 2819, 2821, 2827, and 2829 may be prevented.

Frame 1131 may also include first fastener orifices 2837 arranged about a peripheral area of frame 1131 at one or more intervals. In some embodiments, a pitch between adjacent first fastener orifices 2837 may be constant (or substantially constant), but embodiments are not limited thereto. Second and third fastener orifices 2839 and 2841 may be inset from first fastener orifices 2837 in central portions of frame 1131 respectively near second fluidic inlet and outlet passages 2827 and 2829. A pitch between adjacent second fastener orifices 2839 and a pitch between adjacent third fastener orifices 2841 may be smaller than the pitch(es) between adjacent first fastener orifices 2837. In various embodiments, first, second, and third fastener orifices 2837, 2839, and 2841 may extend completely through frame 1131 and may be counterbored with respect to, for example, surface 2803. When assembled as part of a repeat unit (e.g., repeat unit 1100 in FIG. 11A), first, second, and third fastener orifices 2837, 2839, and 2841 may be configured to respectively receive corresponding fasteners 1137 (see FIG. 11A), which may engage with, for instance, swage nuts 1135 (see FIG. 11A) incorporated into (or as part of) anode frame 1115 (see, e.g., FIGS. 11A and 21), as will become more apparent below. In those instances when frame 1131 is incorporated as part of cathode interface assembly 505 (see, e.g., FIGS. 5-10, 17, and 18)), first, second, and third fastener orifices 2837, 2839, and 2841 may be configured to respectively receive corresponding fasteners 1137 (see FIG. 17), which may engage with, for instance, first, second, and third threaded fastener orifices 4539, 4541, and 4543 of cathode interface separator 1701 (see, e.g., FIGS. 17, 18, and 45), as will become more apparent below.

According to various embodiments, one or more of the counterbored portions of first, second, and third fastener orifices 2837, 2839, and 2841 may be sized to form respective clearance or interference fits with corresponding fasteners 1137 (see FIG. 11A) or corresponding portions (e.g., head or shoulder portions) of fasteners 1137 (see, e.g., FIG. 21) when frame 1131 is assembled as part of a repeat unit (e.g., repeat unit 1100 in FIG. 11A) or as part of cathode interface assembly 505 in, for instance, FIGS. 5-10, 17, and 18. In some embodiments, one or more of the counterbored portions of first, second, and third fastener orifices 2837, 2839, and 2841 may be sized to form respective clearance fits with corresponding fasteners 1137 (see, e.g., FIGS. 11A, 17, and 21) and one or more of the counterbored portions of first, second, and third fastener orifices 2837, 2839, and 2841 may be sized to form respective interference fits with corresponding fasteners 1137. For example, respective widths (e.g., diameters) of the counterbored portions of first, second, and third fastener orifices 2837, 2839, and 2841 may be about 0.01% to about 10% larger (in the case of a clearance fit) or about 0.01% to about 5% smaller (in the case of an interference fit) than corresponding widths (e.g., diameters) of respective portions (e.g., head or shoulder portions) of fasteners 1137 (see, e.g., FIGS. 11A, 17, and 21). In some embodiments, one or more of the counterbored portions of first, second, and third fastener orifices 2837, 2839, and 2841 may be sized to form respective clearance fits with corresponding fasteners 1137 (see, e.g., FIGS. 11A, 17, and 21) or corresponding portions (e.g., head or shoulder portions) of fasteners 1137 (see, e.g., FIG. 21) when frame 1131 is assembled as part of a repeat unit (e.g., repeat unit 1100 in FIG. 11A) or as part of cathode interface assembly 505 in, for instance, FIGS. 5-10, 17, and 18, and stack 500 (see, e.g., FIG. 5) is in a cooled, non-operational state, but expand to form corresponding interference fits in a steady-state operational condition of stack 500. These clearance and/or interference fits may be utilized to constrain in-plane expansion (e.g., expansion in, for instance, a plane parallel to an x-y plane (see FIG. 11A)) of frame 1131 (and, in some embodiments, anode frame 1115 in FIG. 11A) during operation of stack 500 without unduly stressing frame 1131 and/or anode frame 1115. This may prevent (or at least reduce the likelihood of) misalignments, bunching, etc., of anode PTLs 1109 and cathode GDLs 1121 of the various cells/repeat units of stack 500 (see, e.g., FIGS. 5-10), as well as prevent (or reduce the likelihood of) misalignments between adjacent frames of adjacent cells/repeat units of stack 500. Such a configuration may also allow frame 1131 and/or anode frame 1115 to be formed of more compliant materials that, in some cases, may be less expensive and/or easier to manufacture (and, in some cases, not electrically conductive).

According to some embodiments, frame 1131 and/or cathode annular insert 1134 may be formed of any suitable thermoplastic and/or thermosetting material, such as, for instance, polyethylene terephthalate (PET), polycarbonate (PC), polyimide (PI), polyamide (PA), poly(methylmethacrylate) (PMMA), polyethylene naphthalate (PEN), polyetherketone (PEK), polyetheretherketone (PEEK), polystyrene (PS), polyetherimide (PEI), polyphenylene sulfide (PPS), polyarylate (PAR), polyether sulfone (PES), cyclic olefin copolymer (COC), polyvinyl alcohol (PVA), ethylene chlorotrifluoroethylene (ECTFE), polytetrafluoroethylene (PTFE), polybutylene terephthalate (PBT), polychlorotrifluoroethylene (PCTFE), polyethylene terephthalate glycol (PETG), and/or the like. In some cases, frame 1131 and/or cathode annular insert 1134 may be formed of one or more metals or metal alloys, such as aluminum, aluminum alloy, copper, copper alloy, tin, tin alloy, titanium, titanium alloy, tungsten, tungsten alloy, zinc, zinc alloy, steel, stainless steel, etc. It is noted, however, that when formed of a metal or metal alloy, frame 1131 may, in some embodiments, include a coating or other feature to, for instance, electrically insulate frame 1131 from a corresponding cathode GDL (e.g., cathode GDL 1121 in FIG. 11A) and/or cathode flow field (e.g., cathode flow field 1127 in FIG. 11A) associated therewith. It is also contemplated that a base material of frame 1131 may be coated with, for example, one or more other materials, e.g., one or more corrosion-resistant materials. Whatever the case, frame 1131 and/or cathode annular insert 1134 may be formed in any suitable manner, such as additively manufactured, stamped, injection molded, compression molded, casted, machined, and/or the like.

### Anode Frame

Similar to cathode flow field 1127 (see, e.g., FIGS. 11A, 23, and 24), anode flow field 1111 may be at least partially supported in an opening of anode frame 1115 (see, e.g., FIGS. 11A, 23, and 24), which also includes a plurality of fluidic passages to facilitate fluid communication (or flow) through stack 500 (see, e.g., FIGS. 5-10), and, in particular, through a COₓ electrolyzer cell of stack 500, such as cell 501. Various details of an illustrative anode frame 1115 will now be discussed in more detail in association with FIGS. 37-42.

FIG. 37 depicts a first perspective view of an example anode frame. FIG. 38 depicts a top view of the example anode frame of FIG. 37. FIG. 39 depicts a second perspective view of the example anode frame of FIG. 37. FIG. 40 depicts a bottom view of the example anode frame of FIG. 39. FIG. 41 depicts an enlarged portion of the example anode frame of FIG. 38. FIG. 42 depicts an enlarged portion of the example anode frame of FIG. 40.

Anode frame (or frame) 1115 may be a generally rectangular plate-shaped body having first surface 3701 (e.g., a top surface) opposing second surface 3703 (e.g., a bottom surface) in axial direction 3801. Although frame 1115 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, frame 1115 will be described in association with a generally rectangular configuration. First and second surfaces 3701 and 3703 may be bounded by one or more peripheral surfaces, such as peripheral surfaces (or surfaces) 3705, 3707, 3709, and 3711 that may be connected to one another via one or more other peripheral surfaces, such as peripheral surface (or surface) 3713. In some embodiments, frame 1115 may have a symmetrical configuration about one or more reference planes perpendicular to axial direction 3801 (see FIGS. 38 and 40). For instance, a configuration of frame 1115 may be symmetrical about either or both of reference planes 3803 and 3805 depicted in FIGS. 38 and 40, but embodiments are not limited thereto.

According to various embodiments, first fluidic inlet passages 3715 and 3717 may be adjacent to peripheral edge 3705, and first fluidic outlet passages 3719 and 3721 may be adjacent to peripheral edge 3709. First fluidic inlet passages 3715 and 3717 may form portions of inlet passages 1001 and 1003 (see FIG. 10) of stack 500 in association with inlet connectors 543 of manifold assembly 515 (see FIGS. 5-10) that provide input water to frame 1115, and, thereby, to a corresponding anode flow field 1111 (see, e.g., FIGS. 11A, 23, and 24) associated with frame 1115. First fluidic outlet passages 3719 and 3721 may form portions of outlet passages (that are similar to inlet passages 1001 and 1003 (see FIG. 10), but associated with outlet connectors 545 of manifold assembly 515 versus inlet connectors 543 (see, e.g., FIGS. 5-10)) of stack 500 that output water from frame 1115, and, thereby, from the corresponding anode flow field 1111 (see, e.g., FIGS. 11A, 23, and 24) associated with frame 1115. In some implementations, first fluidic inlet and outlet passages 3715-3721 may be defined by respective pluralities of orifices separated from one another via corresponding septal walls. For instance, first fluidic inlet passage 3715 may include first and second inlet orifices 3715a and 3715b separated from one another via septal wall 3701s1, whereas first fluidic outlet passage 3719 may include first and second outlet orifices 3719a and 3719b separated from one another via septal wall 3701s2. An illustrative septal wall is also depicted in the enlarged view of FIG. 42 and the cross-sectional view of FIG. 23. That is, septal wall 3701s3 is shown separating first and second outlet orifices 3721a and 3721b forming first fluidic outlet passage 3721 in FIG. 42, and septal wall 3701s4 is shown separating first and second inlet orifices 3717a and 3717b forming first fluidic inlet passage 3717 in FIG. 23. As with cathode frame 1131 (see, e.g., FIG. 11A), the presence of the septal walls in frame 1115, such as septal walls 3701s1-3701s3, may increase the structural rigidity and, thereby, reliability of frame 1115 in the vicinity of first fluidic inlet and outlet passages 3715-3721.

According to various embodiments, frame 1115 also includes through opening (or opening) 3723 formed completely through a first central portion of frame 1115 and may be configured to receive at least a portion of anode flow field 1111 therein (see, e.g., FIGS. 11A, 23, and 24). As such, opening 3723 may be sized and shaped to correspond with the size and shape of anode flow field 1111. For example, opening 3723 may have a generally rectangular shape with rounded corners, but embodiments are not limited thereto. Frame 1115 may also include blind opening (or opening) 3725 formed in a second central portion of frame 1115 encircling the first central portion of frame 1115. In some cases, opening 3725 may be omitted or may be at least partially filled by anode annular insert 1118, as will become more apparent below. When included as part of frame 1115, opening 3725 may terminate at surface 3701r, which may be recessed from first surface 3701, and may be configured to receive at least a portion of anode PTL 1109 (see, e.g., FIGS. 11A, 23, and 24) and/or at least a portion of anode frame insert 1118 therein. As such, opening 3725 may be sized and shaped to correspond with the size and shape of anode PTL 1109 (see, e.g., FIGS. 11A, 23, and 24) and/or anode frame insert 1118. For instance, opening 3725 may have a generally rectangular shape with rounded corners, but embodiments are not limited thereto. To enable fluid flow to and from anode flow field 1111 (see, e.g., FIGS. 11A, 23, and 24) at least partially supported in opening 3723, first fluidic inlet passages 3715 and 3717 may be fluidically connected to opening 3723 via corresponding channels 4001, 4003, 4005, and 4007, respective connecting risers 3727 and 3729, distribution channel 3731, and supply (or inlet) channels 3733. First fluidic outlet passages 3719 and 3721 may be fluidically connected to opening 3723 via outlet channels 3735, collection channel 3737, respective connecting risers 3739 and 3741, and corresponding channels 4009, 4011, 4013, and 4015.

In those implementations including anode annular insert 1118, anode annular insert 1118 may be at least partially supported in opening 3725 such that second surface 1118b of anode annular insert 1118 abuts against surface 3701r of frame 1115 and inner peripheral surface 1118c of anode annular insert 1118 encircles an outer peripheral boundary of anode flow field 1111, and thereby, an inner peripheral boundary of opening 3723 (see also FIGS. 11B and 11C). To this end, outer peripheral surface 1118d of anode annular insert 1118 may be shaped and sized to correspond with the shape and size of an inner peripheral boundary of opening 3725. In some cases, thickness 1118t of anode annular insert 1118 may be equivalent (or substantially equivalent) to the depth of opening 3725, but implementations are not limited thereto. When thickness 1118t of anode annular insert 1118 corresponds to the depth of opening 3725, anode annular insert 1118 may fill the void in frame 1115 corresponding to opening 3725. It is also contemplated that anode annular insert 1118 may not completely fill the void corresponding to opening 3725, such as can be appreciated in FIGS. 11B and 11C. In such instances, inner peripheral surface 1118c of anode annular insert 1118 may be offset from the inner peripheral boundary of opening 3723 and PTL 1109 may fill a remaining amount of space not filled by anode annular insert 1118. Whatever the case, anode annular insert 1118 may have a generally ring-like configuration, and as such, may not be truly annular. For instance, anode annular insert 1118 may have a generally rectangular cross-section when viewed along the z-axis direction shown in FIGS. 11B and 11C, thus giving rise to an anode annular insert having two-fold symmetry instead of axial symmetry. As such, anode annular insert 1118 may have, for instance, a circular, an oval, a polygonal, or any other suitable cross-sectional geometry when viewed along the z-axis direction shown in FIGS. 11B and 11C.

Inlet and outlet channels 3733 and 3735 may be blind recesses formed in surface 3701r that extend from opening 3723 and terminate at distribution channel 3731 and connecting risers 3727 and 3729 in the case of inlet channels 3733 and distribution channel 3737 and connecting risers 3739 and 3741 in the case of outlet channels 3735, such as illustrated in FIGS. 37, 38, and 41. In some cases, inlet and outlet channels 3733 and 3735 may not only extend parallel (or substantially parallel) to one another, but may also extend parallel (or substantially parallel) to reference plane 3803. When incorporated as part of a cell, such as cell 501, anode annular insert 1118 may be at least partially supported in opening 3725 to at least partially fill the void corresponding to opening 3725. As previously noted, a remaining area of the void may be filled by PTL 1109, and as such, anode annular insert 1118 may serve to extend the outer boundary of PTL 1109 further outwards towards recess 3747 in frame 1115. By filling the void corresponding to opening 3725 (which is formed between opening 3723 and recess 3747) the likelihood that input water that is to be supplied to anode flow field 1111 from inlet channels 3733 instead flows around anode flow field 1111 via opening 3725 (illustrated in FIG. 11B as bypass flow 1120) and becomes expelled via outlet channels 3735 is reduced or eliminated. It is noted that bypass flow 1120 decreases the amount of input water flowing through anode flow field 1111, and as such, has the potential to decrease the efficiency of the cell. In some cases, both opening 3725 and anode annular insert 1118 may be omitted, thereby further reducing the possibility of bypass flow 1120. In those instances when opening 3725 is formed in frame 1115 and anode annular insert 1118 is not utilized, PTL 1109 may be formed to completely (or substantially completely) fill opening 3725 to reduce or prevent the likelihood of bypass flow 1120.

According to some embodiments, the presence of anode annular insert 1118 may not only prevent or reduce the likelihood of bypass flow 1120 during operation of stack 500, but may also prevent or reduce the likelihood that bypass flow 1120 or compression forces within the system (e.g., stack 500) cause the anode side of MEA 1105 to push against the outer periphery of PTL 1109 and become mechanically deteriorated via abrasion, cutting, etc. Anode annular insert 1118 may also prevent or reduce the likelihood that, for instance, first anode gasket 1113a intrudes into one or more of inlet and/or outlet channels 3733 and 3735.

To facilitate distributed supply and collection of water to and from anode flow field 1111 (see, e.g., FIGS. 11A, 23, and 24), inlet and outlet channels may have respective outer channels flanking corresponding central channels. For example, as seen in FIG. 41, outlet channels 3735 may be divided into first outer outlet channels 3735a arranged in first outer portion 4101, second outer outlet channels 3735b arranged in second outer portion 4103, and central outlet channels 3735c arranged in central portion 4105. Central outlet channels 3735c may be spaced apart from one another at constant interval 4107, whereas first and second outer outlet channels 3735a and 3735b may be spaced apart from one another with variable intervals that may increase in size with increasing distance from central portion 4105. For instance, adjacent first outer outlet channels 3735a near central portion 4105 may be spaced apart from one another by interval 4109 and adjacent first outer outlet channels 4135a further away from central portion 4105 may be spaced apart from one another by interval 4111, which may be greater than interval 4109. Inlet channels 3733 may be similarly arranged and configured as outlet channels 3735, but with respect to an inlet side of opening 3723 versus the outlet side of opening 3723 associated with outlet channels 3735.

The central inlet and outlet channels (e.g., central outlet channels 3735c) of inlet and outlet channels 3733 and 3735 may respectively terminate at and be fluidically connected to distribution channels 3731 and 3737. Some of the first outer inlet and outlet channels of inlet and outlet channels 3733 and 3735 may respectively terminate at and be fluidically connected to distribution channels 3731 and 3737, whereas other ones of the first outer inlet and outlet channels (e.g., the identified first outer outlet channels 3735a in FIG. 41) of inlet and outlet channels 3733 and 3735 may respectively terminate at and be fluidically connected to connecting risers 3727 and 3741. Similarly, some of the second outer inlet and outlet channels of inlet and outlet channels 3733 and 3735 may respectively terminate at and be fluidically connected to distribution channels 3731 and 3737, whereas other ones of the second outer inlet and outlet channels (e.g., the identified second outer outlet channels 3735b in FIG. 41) of inlet and outlet channels 3733 and 3735 may respectively terminate at and be fluidically connected to connecting risers 3729 and 3739.

Distribution channels 3731 and 3737 may be formed as blind recesses in surface 3701r and may extend in a direction transverse to the direction of extension of inlet and outlet channels 3735, such as depicted in FIGS. 37, 38, and 41. In some embodiments, distribution channels 3731 and 3737 may extend parallel (or substantially parallel) to reference plane 3805. Distribution channel 3731 may be flanked on either side by and fluidically connected to connecting risers 3727 and 3729, which may be formed as orifices extending through frame 1115 from surface 3701r to surface 3703 in axial direction 3801, such as can be appreciated from FIGS. 37-42. Similarly, distribution channel 3737 may be flanked on either side by and fluidically connected to connecting risers 3739 and 3741, which may be formed as orifices extending through frame 1115 from surface 3701r to surface 3703 in axial direction 3801.

As seen in FIGS. 39 and 40, connecting risers 3727, 3729, 3739, and 3749 may be fluidically connected to first fluidic inlet and outlet passages 3715-3721, respectively, via corresponding groups of channels 4001-4015. For instance, connecting riser 3727 may be fluidically connected to first fluidic inlet passages 3715 via channels 4001 and 4003, whereas connecting riser 3729 may be fluidically connected to first fluidic inlet passages 3717 via channels 4005 and 4007. Further, connecting riser 3739 may be fluidically connected to first fluidic outlet passages 3719 via channels 4009 and 4011, whereas connecting riser 3741 may be fluidically connected to first fluidic outlet passages 3721 via channels 4013 and 4015.

Channels 4001-4015 may be formed as blind recesses in surface 3703 and may extend in oblique directions with respect to, for instance, a direction of extension of reference plane 3803, as can be appreciated in FIGS. 39, 40, and 42. For instance, as seen in FIG. 42, channels 4015 may not only extend parallel (or substantially parallel) to one another, but may extend from first outlet orifice 3721a of first fluidic outlet passage 3721 to connecting riser 3741 at oblique angle 4201. Similarly, channels 4013 may not only extend parallel (or substantially parallel) to one another, but may extend from second outlet orifice 3721b of first fluidic outlet passage 3721 to connecting riser 3741 at oblique angle 4203, which may be smaller than oblique angle 4201. In some embodiments, channels 4013 and 4015 may be formed as respective groups of six channels, but embodiments are not limited thereto. For example, any number of channels may be utilized, such as less or more than six. Additionally, channels 4013 and 4015 may have the same number of individual channels or a different number of individual channels. To this end, the individual channels among channels 4013 and 4015 may have equivalent (or substantially equivalent) cross-sectional areas in a plane perpendicular to their respective directions of longitudinal extension. In some embodiments, some of the individual channels may have equivalent (or substantially equivalent) cross-sectional areas (such as channels 4013a and 4013b) and at least one of the individual channels may have a different cross-sectional area (such as channel 4013c). In the case of individual channel 4013c, its cross-sectional area may vary in size, such as increase in cross-sectional area with increasing distance from second outlet orifice 3721b of first fluidic outlet passage 3721. Channels 4001-4011 may be similarly configured as described in association with channels 4013 and 4015, but with respect to the corresponding connecting risers and first fluidic inlet and outlet passages associated therewith.

According to various embodiments, openings 3723 and 3725 may be arranged between second fluidic inlet and outlet passages 3743 and 3745, which form respective portions of inlet and outlet passages 901 and 903 (see FIG. 9) of stack 500 in association with input and outlet connectors 547 and 549 of manifold assembly 515 (see, e.g., FIGS. 5-10). Inlet passage 901 (see FIG. 9) may supply one or more reactants (e.g., gaseous COₓ) to the various cathode frames 1131 of stack 500 (see, e.g., FIG. 5), and, as such, to the corresponding cathode flow fields 1127 (see, e.g., FIGS. 5-11A) supported in association therewith when frame 1115 is incorporated as part of a cell, such as cell 501. Outlet passage 903 (see FIG. 9), however, may enable one or more byproducts of the COₓ reduction process to be expelled from the various cathode frames 1131 of stack 500 (see, e.g., FIGS. 5-11A), and, thereby, from the corresponding cathode flow fields 1127 supported in association therewith.

Frame 1115 may also include recesses 3747-3759 in surface 3701 that may be configured to respectively receive corresponding portions of gaskets among first anode gasket set 1113 (see, e.g., FIGS. 11A, 23, and 24) therein when, for example, frame 1115 is assembled as part of a repeat unit (e.g., repeat unit 503_1 in FIG. 5) or anode interface assembly 509 (see, e.g., FIGS. 5-10, 47, and 48). For instance, and with momentary reference to FIGS. 11A, 23, and 24 in addition to FIGS. 37-42, recess 3747 may be formed to encircle the periphery of opening 3725 and interface with first anode gasket 1113a of first anode gasket set 1113, whereas recesses 3749-3755 may be formed to respectively encircle the peripheries of first fluidic inlet and outlet passages 3715-3721 and respectively interface with second anode gaskets 1113b of first anode gasket set 1113. It is noted that the conjunction of first fluidic inlet passages 3715 and 3717, channels 4001, 4003, 4005, and 4007, connecting risers 3727 and 3729, distribution channel 3731, and supply channels 3733 enables, for example, water to flow from an area outside of first anode gasket 1113a of first anode gasket set 1113 (see, e.g., FIGS. 11A, 23, and 24) to an area inside of first anode gasket 1113a of first anode gasket set 1113 without disturbing the integrity of or seal provided by first anode gasket 1113a of first anode gasket set 1113. The same is true with respect to the integrity of and seals provided by those second anode gaskets 1113b of first anode gasket set 1113 that interface with recesses 3749 and 3751, see, e.g., FIGS. 11A, 23, and 24). In a similar fashion, the conjunction of first fluidic outlet passages 3719 and 3721, outlet channels 3735, collection channel 3737, connecting risers 3739 and 3741, and channels 4009, 4011, 4013, and 4015 enables, for example, water to flow from an area inside of first anode gasket 1113a of first anode gasket set 1113 (see, e.g., FIGS. 11A, 23, and 24) to an area outside of first anode gasket 1113a of first anode gasket set 1113 without disturbing the integrity of or seal provided by first anode gasket 1113a of first anode gasket set 1113. The same is true with respect to the integrity of and seals provided by those second anode gaskets 1113b of first anode gasket set 1113 (see, e.g., FIGS. 11A, 23, and 24) that interface with recesses 3753 and 3755. In addition, recesses 3757 and 3759 may be formed to encircle the respective peripheries of second fluidic inlet and outlet passages 3743 and 3745 and interface with third anode gaskets 1113c of first anode gasket set 1113 (see, e.g., FIGS. 11A, 23, and 24).

Similar to recesses 3747-3759 formed in surface 3701, frame 1115 may include recesses 4017-4029 in surface 3703 that may be configured to respectively receive corresponding portions of gaskets among second anode gasket set 1117 (see, e.g., FIGS. 11A, 23, and 24) therein when, for example, frame 1115 is assembled as part of a repeat unit (e.g., repeat unit 503_1 in FIG. 5) or anode interface assembly 509 (see, e.g., FIGS. 5-10, 47, and 48). For instance, recess 3717 may be formed to encircle the periphery of opening 3723 and interface with first anode gasket 1117a of second anode gasket set 1117 (see, e.g., FIGS. 11A, 23, and 24). Recesses 4019-4025 may be formed to respectively encircle combined peripheries of associated first fluidic inlet and outlet passages 3715-3721, corresponding channels 4001-4015, and respective connecting risers 3727, 3729, 3739, and 3741 and respectively interface with second anode gaskets 1117b of second anode gasket set 1117 (see, e.g., FIGS. 11A, 23, and 24). For example, recess 4019 may be formed to encircle a combined periphery of first fluidic inlet passages 3717, channels 4005 and 4007, and connecting riser 3729 and to interface with one of second anode gaskets 1117b of second anode gasket set 1117 (see, e.g., FIGS. 11A, 23, and 24), whereas recess 4021 may be formed to encircle a combined periphery of first fluidic inlet passages 3715, channels 4001 and 4003, and connecting riser 3727 to interface with another one of second anode gaskets 1117b of second anode gasket set 1117 (see, e.g., FIGS. 11A, 23, and 24). Similarly, recess 4023 may be formed to encircle a combined periphery of first fluidic outlet passages 3721, channels 4013 and 4015, and connecting riser 3741 to interface with still another one of second anode gaskets 1117b of second anode gasket set 1117 (see, e.g., FIGS. 11A, 23, and 24), whereas recess 4025 may be formed to encircle a combined periphery of first fluidic outlet passages 3719, channels 4009 and 4011, and connecting riser 3739 to interface with yet another one of second anode gaskets 1117b of second anode gasket set 1117 (see, e.g., FIGS. 11A, 23, and 24). It is noted that the conjunction of first fluidic inlet passages 3715 and 3717, channels 4001, 4003, 4005, and 4007, connecting risers 3727 and 3729, distribution channel 3731, and supply channels 3733 enables, for example, water to flow from an area outside of first anode gasket 1113a of first anode gasket set 1113 (see, e.g., FIGS. 11A, 23, and 24) to an area inside of first anode gasket 1113a of first anode gasket set 1113 without also disturbing the integrity of or seal provided by second anode gaskets 1117b of second anode gasket set 1117 (see, e.g., FIGS. 11A, 23, and 24). In addition, recesses 4027 and 4029 may be formed to at least encircle the respective peripheries of second fluidic inlet and outlet passages 3743 and 3745 and interface with third anode gaskets 1117c of second anode gasket set 1117 (see, e.g., FIGS. 11A, 23, and 24). It is noted that the size, shape, and location of recesses 4019-4029 may correspond with the size, shape, and location of protrusions 3305 and 3307 (see FIGS. 32-36) of cathode frame 1131 to enable second and third anode gaskets 1117b and 1117c (see, e.g., FIGS. 11A, 23, and 24) to form corresponding seals between anode and cathode frames 1115 and 1131 when anode and cathode frames 1115 and 1131 are stacked in relation with other anode and cathode frames 1115 and 1131 of stack 500 (see, e.g., FIGS. 5-11A, 23, and 24). Accordingly, cross-flow between first and second fluidic inlet and outlet passages 3715-3721, 3743, and 3745 may be prevented.

Frame 1115 may also include first fastener orifices 3761 arranged about a peripheral area of frame 1115 at one or more intervals. In some embodiments, a pitch between adjacent first fastener orifices 3761 may be constant (or substantially constant), but embodiments are not limited thereto. Second and third fastener orifices 3763 and 3765 may be inset from first fastener orifices 3761 in central portions of frame 1115 near second fluidic inlet and outlet passages 3743 and 3745. A pitch between adjacent second fastener orifices 3763 and a pitch between adjacent third fastener orifices 3765 may be smaller than the pitch(es) between adjacent first fastener orifices 3761. In various embodiments, first, second, and third fastener orifices 3761, 3763, and 3765 may extend completely through frame 1115 and may be counterbored with respect to surface 3701. According to various embodiments, swage nuts 1135 (see, e.g., FIGS. 11A and 21) may be pressed into, for example, the counterbored portions of first, second, and third fastener orifices 3761, 3763, and 3765 such that, when frame 1115 is assembled as part of a repeat unit (e.g., repeat unit 503_1 in FIG. 5) or as part of anode interface assembly 509 (see, e.g., FIGS. 5-10, 47, and 48), first, second, and third fastener orifices 3761, 3763, and 3765 may be configured to respectively engage with corresponding fasteners 1137 (see, e.g., FIGS. 11A and 21), which may be received in corresponding first, second, and third fastener orifices 2837, 2839, and 2841 of cathode frame 1131 (see, e.g., FIGS. 11A, 21, 28, 29, 32, 33, and 35).

According to some embodiments, frame 1115 and/or anode annular insert 1118 may be formed of any suitable thermoplastic and/or thermosetting material, such as, for instance, PET, PC, PI, PA, PMMA, PEN, PEK, PEEK, PEI, PPS, PAR, PES, COC, PVA, PS, ECTFE, PTFE, PBT, PCTFE, PETG, and/or the like. In some cases, frame 1115 and/or anode annular insert 1118 may be formed of one or more metals or metal alloys, such as, for example, aluminum, aluminum alloy, copper, copper alloy, tin, tin alloy, titanium, titanium alloy, tungsten, tungsten alloy, zinc, zinc alloy, steel, stainless steel, etc. It is noted, however, that when formed of a metal or metal alloy, frame 1115 and/or anode annular insert 1118 may, in some embodiments, include a coating or other feature to, for instance, electrically insulate frame 1115 or anode annular insert 1118 from a corresponding anode PTL (e.g., anode PTL 1109 in FIG. 11A) and/or anode flow field (e.g., anode flow field 1111 in FIG. 11A) associated therewith. It is also contemplated that a base material of frame 1131 and/or anode annular insert 1118 may be coated with, for instance, one or more other materials, e.g., one or more corrosion-resistant materials. That being said, in some cases, anode annular insert 1118 may be formed of one or more materials with equivalent, substantially equivalent, or at least similar chemical inertness as PTL 1109. To this end, anode annular insert 1118 may have a porous or non-porous configuration. Whatever the case, frame 1115 and/or anode annular insert 1118 may be formed in any suitable manner, such as additively manufactured, injection molded, compression molded, stamped, casted, machined, and/or the like.

### Separator Plate

FIG. 43 depicts a plan view of an example separator plate of the representative repeat unit of FIG. 11A.

Separator plate 1107 may be a generally rectangular plate-shaped body having first surface 4301 (e.g., a top surface) opposing a second surface in axial direction 4303. Although separator plate 1107 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, separator plate 11070 will be described in association with a generally rectangular configuration. First surface 4301 and the second surface may be bounded by one or more peripheral surfaces, such as peripheral surfaces (or surfaces) 4305, 4307, 4309, and 4311 that may be connected to one another via one or more other peripheral surfaces, such as peripheral surface (or surface) 4313. Separator plate 1107 may also have terminal 4307t protruding from peripheral surface 4307. It is noted that when corresponding separator plates (such as separator plate 1107) are interposed between adjacent cells among stack 500 (see FIGS. 5-10), corresponding voltage drops between adjacent separator plates (and, thereby, associated with respective cells correspondingly between the adjacent separator plates) may be probed via respective terminals (such as terminal 4307t) of the corresponding separator plates, such as separator plate 1107 (see also FIG 7). In some embodiments, separator plate 1107 may have a symmetrical configuration about one or more reference planes perpendicular to axial direction 4303. For instance, a configuration of separator plate 1107 may be symmetrical about either or both of reference planes 4315 and 4317 (apart from the presence of terminal 4307t), but embodiments are not limited thereto.

According to various implementations, separator plate 1107 includes first openings 4319 and 4321 adjacent to peripheral surface 4305, second openings 4323 and 4325 adjacent to peripheral surface 4309, third opening 4327 adjacent to peripheral surface 4305, and fourth opening 4329 adjacent to peripheral surface 4309. Openings 4319 and 4321 may be sized, shaped, and located in correspondence with the size, shape, and location of protrusions 3305 (see, e.g., FIGS. 32 and 33) adjacent to peripheral surface 2805 of cathode frame 1131 such that, when separator plate 1107 is incorporated as part of a repeat unit (e.g., repeat unit 1100 in FIG. 11A), protrusions 3305 adjacent to peripheral surface 2805 of cathode frame 1131 may be received in openings 4319 and 4321 (see also FIG. 23). Similarly, openings 4323 and 4325 may be sized, shaped, and located in correspondence with the size, shape, and location of protrusions 3305 adjacent to peripheral surface 2809 of cathode frame 1131 (see, e.g., FIGS. 32 and 33) such that, when separator plate 1107 is incorporated as part of a repeat unit (e.g., repeat unit 1100 in FIG. 11A), protrusions 3305 adjacent to peripheral surface 2809 of cathode frame 1131 may be received in openings 4323 and 4325. Further, openings 4327 and 4329 may be sized, shaped, and located in correspondence with the size, shape, and location of protrusions 3307 adjacent to peripheral surfaces 2805 and 2809 of cathode frame 1131 (see, e.g., FIGS. 24, 32, and 33) such that, when separator plate 1107 is incorporated as part of a repeat unit (e.g., repeat unit 1100 in FIG. 11A), protrusions 3307 adjacent to peripheral surfaces 2805 and 2809 of cathode frame 1131 may be respectively received in openings 4327 and 4329 (see also FIG. 24). Relative dimensioning between openings 4319-4329 and first and second protrusions 3305 and 3307 has already been described in association with cathode frame 1131, and, therefore, duplicative descriptions will be omitted to avoid obscuring embodiments described herein. In this manner, first surface 4301 of separator plate 1107 may abut against surface 3701 of anode frame 1115 (see, e.g., FIGS. 23, 24, 37, and 38) and the second surface of separator plate 1107 may abut against surface 2801 of cathode frame 1131 (see, e.g., FIGS. 23, 24, 32, and 33) when the repeat unit (e.g., repeat unit 1100 in FIG. 11A) is assembled, such as assembled in a compressed state (see also FIGS. 20-24).

Separator plate 1107 may also include first fastener orifices 4331 arranged about a peripheral area of separator plate 1107 at one or more intervals. In some embodiments, a pitch between adjacent first fastener orifices 4331 may be constant (or substantially constant), but embodiments are not limited thereto. Second and third fastener orifices 4333 and 4335 may be inset from first fastener orifices 4331 in central portions of separator plate 1107 near third and fourth openings 4327 and 4329. A pitch between adjacent second fastener orifices 4333 and a pitch between adjacent third fastener orifices 4335 may be smaller than the pitch(es) between adjacent first fastener orifices 4331. In various embodiments, first, second, and third fastener orifices 4331, 4333, and 4335 may extend completely through separator plate 1107 such that, when separator plate 1107 is assembled as part of a repeat unit (e.g., repeat unit 1100 in FIG. 11A), fasteners 1137 extending from cathode frame 1131 may extend through separator plate 1107 and may be threadedly engaged with corresponding swage nuts 1135 pressed and/or clinched into first, second, and third fastener orifices 3761, 3763, and 3765 of anode frame 1115 (see also FIGS. 11A and 21).

According to various embodiments, one or more of first, second, and third fastener orifices 4331, 4333, and 4335 may be sized to form respective clearance or interference fits with corresponding fasteners 1137 (see FIG. 11A) or corresponding portions (e.g., shoulder portions) of fasteners 1137 (see, e.g., FIG. 21) when separator plate 1107 is assembled as part of a repeat unit (e.g., repeat unit 1100 in FIG. 11A). In some cases, one or more of first, second, and third fastener orifices 4331, 4333, and 4335 may be sized to form respective clearance fits with corresponding fasteners 1137 (see FIG. 11A) or corresponding portions (e.g., shoulder portions) of fasteners 1137 (see, e.g., FIG. 21) and one or more of first, second, and third fastener orifices 4331, 4333, and 4335 may be sized to form respective interference fits with corresponding fasteners 1137 (see FIG. 11A) or corresponding portions (e.g., shoulder portions) of fasteners 1137 (see, e.g., FIG. 21). For example, respective sizes (e.g., diameters) of first, second, and third fastener orifices 4331, 4333, and 4335 may be about 0.01% to about 10% larger (in the case of a clearance fit) or about 0.01% to about 5% smaller (in the case of an interference fit) than corresponding widths (e.g., diameters) of respective portions (e.g., shoulder portions) of fasteners 1137 (see, e.g., FIGS. 11A, 17, and 21). In some embodiments, one or more of first, second, and third fastener orifices 4331, 4333, and 4335 may be sized to form respective clearance fits with corresponding fasteners 1137 (see, e.g., FIGS. 11A, 17, and 21) or corresponding portions (e.g., shoulder portions) of fasteners 1137 (see, e.g., FIG. 21) when separator plate 1107 is assembled as part of a repeat unit (e.g., repeat unit 1100 in FIG. 11A) and stack 500 (see, e.g., FIG. 5) is in a cooled, non-operational state, but when stack 500 is in a steady-state operational condition, fasteners 1137 may expand to form corresponding interference fits with the one or more of first, second, and third fastener orifices 4331, 4333, and 4335. These clearance and/or interference fits may be utilized to constrain in-plane expansion (e.g., expansion in, for instance, a plane parallel to an x-y plane (see FIG. 11A)) of anode and cathode frames 1115 and 1131 during operation of stack 500 (see, e.g., FIG. 5) without unduly stressing anode and cathode frames 1115 and 1131.

It is also noted that, when separator plate 1107 is assembled as part of a repeat unit (e.g., repeat unit 1100 in FIG. 11A) with cathode frame 1131 coupled to anode frame 1115 via fasteners 1137 and swage nuts 1135 (see also FIGS. 11A and 21-24), some of the various gaskets of second anode gasket set 1117 may not only be interposed between surface 4301 of separator plate 1107 and some of the various recesses in surface 3703 of anode frame 1115 (see, e.g., FIGS. 39 and 40), but may also encircle the various protrusions extending from surface 2801 of cathode frame 1131 (see, e.g., FIGS. 32 and 33). For example, second gaskets 1117b of second anode gasket set 1117 (see, e.g., FIGS. 11A and 23) may not only be interposed between surface 4301 of separator plate 1107 and corresponding recesses 4019-4025 in surface 3703 of anode frame 1115 (see also FIGS. 39 and 40), but may also encircle protrusions 3305 extending from surface 2801 of cathode frame 1131 (see also FIGS. 32 and 33) to fluidically seal corresponding first fluidic inlet and outlet passageways between cathode frame 1131 and anode frame 1115 (see, e.g., second anode gasket 1117b fluidically sealing first fluidic inlet passageway 2301 that is outlined in FIG. 23 in a dash-dot-dot line format). In a similar fashion, third gaskets 1117c of second anode gasket set 1117 (see, e.g., FIGS. 11A and 24) may not only be interposed between surface 4301 of separator plate 1107 and corresponding recesses 4027-4029 in surface 3703 of anode frame 1115 (see also FIGS. 39 and 40), but may also encircle protrusions 3307 extending from surface 2801 of cathode frame 1131 (see also FIGS. 32 and 33) to fluidically seal corresponding second fluidic inlet and outlet passageways between cathode frame 1131 and anode frame 1115 (see, e.g., third anode gasket 1117c fluidically sealing second fluidic outlet passageway 2401 that is outlined in FIG. 24 in a dash-dot-dot line format).

According to various embodiments, separator plate 1107 may be formed of any suitable thermoplastic and/or thermosetting material, such as, for instance, PET, PC, PI, PA, PMMA, PEN, PEK, PEEK, PEI, PPS, PAR, PES, COC, PVA, PS, ECTFE, PTFE, PBT, PCTFE, PETG, and/or the like. In some cases, separator plate 1107 may be formed of one or more metals or metal alloys, such as, for example, aluminum, aluminum alloy, copper, copper alloy, tin, tin alloy, titanium, titanium alloy, tungsten, tungsten alloy, zinc, zinc alloy, steel, stainless steel, etc. For instance, in one embodiment, separator plate 1107 may be formed of titanium, which may increase the strength and rigidity of a repeat unit, such as repeat unit 1100 in FIG. 11A, as well as enable electrical conductivity between adjacent cells of stack 500 (see, e.g., FIGS. 5 and 7). In some embodiments, a material(s) and/or configuration of separator plate 1107 may be stronger and/or more rigid than a material(s) and/or configuration of anode and cathode frames 1115 and 1131 (see also FIG. 1 1A). In some instances, an electrical conductivity of separator plate 1107 may be greater than corresponding electrical conductivities of anode and cathode frames 1115 and 1131 (see also FIG. 11A). It is also contemplated that a base material of separator plate 1107 may be coated with, for instance, one or more other materials, e.g., one or more corrosion-resistant materials. Whatever the case, separator plate 1107 may be formed in any suitable manner, such as additively manufactured, injection molded, compression molded, stamped, casted, machined, and/or the like.

### Cathode Interface Assembly

FIG. 17 depicts an exploded view of an example cathode interface assembly of the example multi-cell COₓ electrolyzer stack of FIG. 6. FIG. 18 depicts the example cathode interface assembly of FIG. 17 in a non-exploded state. FIGS. 45 and 46 depict top and bottom plan views of an example cathode interface separator of the example cathode interface assembly of FIG. 18.

As seen in FIGS. 5-10, 17, and 18, cathode interface assembly 505 may include equivalent components as cathode components 1103 of repeat unit 1100 described in association with FIG. 11A, except cathode interface assembly 505 may also include cathode interface separator 1701, third cathode gaskets 1703, and fourth cathode gaskets 1705. As such, duplicative descriptions of equivalent components will be omitted to avoid obscuring embodiments disclosed herein. It is noted, however, that instead of cathode frame 1131 being coupled to anode frame 1115 as in repeat unit 1100 (see FIG. 11A), cathode frame 1131 may be coupled to cathode interface separator 1701, which will now be described in more detail in association with FIGS. 45 and 46.

Referring to FIGS. 45 and 46, cathode interface separator 1701 may be a generally rectangular plate-shaped body having first surface 4501 (e.g., a top surface) opposing second surface 4503 (e.g., a bottom surface) in axial direction 4601. Although cathode interface separator 1701 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, cathode interface separator 1701 will be described in association with a generally rectangular configuration. First and second surfaces 4501 and 4503 may be bounded by one or more peripheral surfaces, such as peripheral surfaces (or surfaces) 4505, 4507, 4509, and 4511 that may be connected to one another via one or more other peripheral surfaces, such as peripheral surface (or surface) 4513. In some embodiments, cathode interface separator 1701 may have a symmetrical configuration about one or more reference planes perpendicular to axial direction 4601. For instance, a configuration of cathode interface separator 1701 may be symmetrical about either or both of reference planes 4603 and 4605, but embodiments are not limited thereto.

According to various embodiments, cathode interface separator 1701 may include first fluidic inlet passages 4515 and 4517 adjacent to peripheral edge 4505, and first fluidic outlet passages 4519 and 4521 adjacent to peripheral edge 4509. With additional reference to FIGS. 5-11A, first fluidic inlet passages 4515 and 4517 may form portions of inlet passages 1001 and 1003 of stack 500 in association with inlet connectors 543 of manifold assembly 515 that provide, for example, input water to anode frames 1115 of stack 500, and, thereby, to the corresponding anode flow fields 1111 of the plurality of cells, such as cell 501. First fluidic outlet passages 4519 and 4521 may form portions of outlet passages (that are similar to inlet passages 1001 and 1003, but associated with outlet connectors 545 of manifold assembly 515 versus inlet connectors 543) of stack 500 that output water from anode frames 1115, and, thereby, from corresponding anode flow fields 1111 of the plurality of cells, such as cell 501 (see also FIGS. 5-11A). In some implementations, first fluidic inlet and outlet passages 4515-4521 may be defined by respective pluralities of orifices separated from one another via corresponding septal walls. For instance, first fluidic inlet passage 4515 may include first and second inlet orifices 4515a and 4515b separated from one another via septal wall 4501s1, whereas first fluidic outlet passage 4519 may include first and second outlet orifices 4519a and 4519b separated from one another via septal wall 4501s2. As with anode and cathode frames 1115 and 1131 (see, e.g., FIG. 11A), the presence of these septal walls, such as septal walls 4501s1 and 4501s2, may increase the structural rigidity and, thereby, reliability of cathode interface separator 1701 in the vicinity of first fluidic inlet and outlet passages 4515-4521.

Cathode interface separator 1701 may further include second inlet and outlet passages 4523 and 4525, which form respective portions of inlet and outlet passages 901 and 903 of stack 500 (see FIG. 9) in association with input and outlet connectors 547 and 549 of manifold assembly 515 (see, e.g., FIGS. 5 and 9). Inlet passage 901 (see FIG. 9) may supply one or more reactants (e.g., gaseous COₓ) to the various cathode frames 1131 of stack 500 (see, e.g., FIGS. 5 and 9), and, as such, to the corresponding cathode flow fields 1127 supported in association therewith when cathode interface separator 1701 is incorporated as part of a cell, such as a cell formed between cathode interface assembly 505 and repeat unit 503_1 (see, e.g., FIGS. 5-11A and 19). Outlet passage 903, however, may enable one or more byproducts of the COₓ reduction process to be expelled from the various cathode frames 1131 of stack 500, and, thereby, from the corresponding cathode flow fields 1127 supported in association therewith (see, e.g., FIGS. 5-11A and 19).

Similar to anode frame 1115 (see, e.g., FIGS. 11A, 37, and 38), cathode interface separator 1701 may also include recesses 4527-4537 in surface 4501 that may be configured to respectively receive corresponding portions of gaskets 553 and 555 when, for example, cathode interface assembly 505 is assembled as part of stack 500, e.g., when cathode interface assembly 505 is stacked in relation to manifold assembly 515 with bus plate 513 interposed therebetween (see, e.g., FIGS. 5-10, 17, and 18). For instance, recesses 4527-4533 may be formed to respectively encircle the peripheries of first fluidic inlet and outlet passages 4515-4521 and respectively interface with corresponding gaskets 553 (which may respectively encircle third fluidic outlet and inlet ports 1225 and 1229 of manifold assembly 515 (see, e.g., FIG. 12)), whereas recesses 4535 and 4537 may be formed to respectively encircle the peripheries of second fluidic inlet and outlet passages 4535 and 4537 and respectively interface with corresponding gaskets 555 (which may respectively encircle fourth fluidic outlet and inlet ports 1239 and 1237 of manifold assembly 515 (see, e.g., FIG. 12)). As such, corresponding fluidic seals may be formed with respective outlet and inlet ports of manifold assembly 515 when cathode interface assembly 505 is assembled as part of stack 500 (see, e.g., FIGS. 5-10).

Referring to FIG. 46, second surface 4503 may include first recesses 4607-4613 respectively encircling first fluidic inlet and outlet passages 4515-4521, as well as second recesses 4615 and 4617 respectively encircling second fluidic inlet and outlet passages 4535 and 4537. In some embodiments, first and second recesses 4607-4617 may be recessed into surface 4503 by a depth equivalent (or substantially equivalent) to height 3401 (see FIG. 34) of first and second protrusions 3305 and 3307 of cathode frame 1131, but embodiments are not limited thereto. For instance, the depth at which first and second recessed 4607-4617 extend into surface 4503 may be greater than or smaller than height 3401 (see FIG. 34) provided sufficient fluidic seals may be formed between cathode interface separator 1701 and cathode frame 1131 when a cell is formed between cathode interface assembly 505 and repeat unit 503_1 (see also FIGS. 5-10 and 17). In other words, the depth of first and second recesses 4607-4617 may at least permit a portion of first and second protrusions 3305 and 3307 of cathode frame 1131 to be received therein when a cell is formed between cathode interface assembly 505 and repeat unit 503_1 (see also FIGS. 5-10). With this in mind, first and second recesses 4607-4613 may be sized and shaped to interface with corresponding protrusions among first and second protrusions 3305 and 3307 of cathode frame 1131 (see FIGS. 32-33).

Cathode interface separator 1701 may further include third recesses 4619-4625 in surface 4503 respectively encircling first fluidic inlet and outlet passages 4515-4521 and associated recesses 4607-4613, as well as include fourth recesses 4627 and 4629 respectively encircling second fluidic inlet and outlet passages 4523 and 4525 and associated recesses 4615-4617. It is also noted that third and fourth recesses 4619-4629 may be respectively sized, shaped, and located to further correspond with the size, shape, and location of protrusions 3305 and 3307 of cathode frame 1131 (see FIGS. 32-33) to enable third and fourth cathode gaskets 1703 and 1705 to form corresponding seals between cathode interface separator 1701 and first and second protrusions 3305 and 3307 of cathode frame 1131 when a cell is formed between cathode interface assembly 505 and repeat unit 503_1 (see also FIGS. 5-10, 32, and 33). Accordingly, the conjunction of first and second recesses 4607-4617 of cathode interface separator 1701, third and fourth recesses 4619-4629 of cathode interface separator 1701, first and second protrusions 3305 and 3307 of cathode frame 1131 (see FIGS. 32-33), and third and fourth cathode gaskets 1703 and 1705 may prevent cross-flow between first and second fluidic inlet and outlet passages 4515-4525. It is also noted that, when a cell is formed between cathode interface assembly 505 and repeat unit 503_1 (see, e.g., FIGS. 5-10), second cathode gasket 1133 may be interposed between a central portion of surface 4503 and recess 3303 in cathode frame 1131 (see FIGS. 17, 32, and 33) to form a fluidic seal around cathode flow field 1127 at least partially supported in an opening of cathode frame 1131. In this manner, corresponding surfaces of cathode flow field 1127 may abut against surface 4503 of cathode interface separator 1701 and a surface of cathode GDL 1121 facing cathode flow field 1127 similar to how corresponding surfaces of cathode flow field 1127 may abut against a surface of cathode GDL 1121 of unitized MEA assembly 1119 and a surface of separator plate 1107 described in association with, for instance, FIGS. 5-11A, 23, and 24.

Cathode interface separator 1701 may also include first threaded fastener orifices 4539 arranged about a peripheral area of cathode interface separator 1701 at one or more intervals. In some embodiments, a pitch between adjacent first threaded fastener orifices 4539 may be constant (or substantially constant), but embodiments are not limited thereto. Cathode interface separator 1701 may optionally include second and third threaded fastener orifices 4541 and 4543 inset from first threaded fastener orifices 4539 in central portions of cathode interface separator 1701 near second fluidic inlet and outlet passages 4523 and 4525. A pitch between adjacent second threaded fastener orifices 4541 and a pitch between adjacent third threaded fastener orifices 4543 may be smaller than the pitch(es) between adjacent first threaded fastener orifices 4539. In some embodiments, one or more of first, second, and third threaded fastener orifices 4539-4543 may be formed similar to first, second, and third fastener orifices 3761-3765 of anode frame 1115 (see, e.g., FIGS. 11A and 37-42), and, thereby, include swage nuts 1135 versus being threaded. Regardless, when cathode interface separator 1701 is assembled as part of cathode interface assembly 505 (see also FIGS. 5-10), first, second, and third threaded fastener orifices 4539, 4541, and 4543 may be configured to respectively engage with corresponding fasteners 1137 respectively received in and extending from corresponding first, second, and third fastener orifices 2837, 2839, and 2841 of cathode frame 1131 (see FIGS. 28, 29, 32, 33, and 35). Further, as can be appreciated from at least FIG. 17, cathode frame 1131 of cathode interface assembly 505 may be coupled to cathode interface separator 1701 with second, third, and fourth cathode gaskets 1133, 1703, and 1705 interposed therebetween.

According to various embodiments, cathode interface separator 1701 may be formed of any suitable thermoplastic and/or thermosetting material, such as, for instance, PET, PC, PI, PA, PMMA, PEN, PEK, PEEK, PEI, PPS, PAR, PES, COC, PVA, PS, ECTFE, PTFE, PBT, PCTFE, PETG, and/or the like. In some cases, cathode interface separator 1701 may be formed of one or more metals or metal alloys, such as, for example, aluminum, aluminum alloy, copper, copper alloy, tin, tin alloy, titanium, titanium alloy, tungsten, tungsten alloy, zinc, zinc alloy, steel, stainless steel, etc. For instance, in one embodiment, cathode interface separator 1701 may be formed of titanium, which may increase the strength and rigidity of cathode interface assembly 505 (see, e.g., FIGS. 5-10, 17, and 18). In some cases, a material(s) and/or configuration of cathode interface separator 1701 may be stronger and/or more rigid than a material(s) and/or configuration of anode and cathode frames 1115 and 1131 (see also FIG. 11A). Also, an electrical conductivity of cathode interface separator 1701 may, in some embodiments, be greater than corresponding electrical conductivities of anode and cathode frames 1115 and 1131 (see also FIG. 11A). It is also contemplated that a base material of cathode interface separator 1701 may be coated with, for instance, one or more other materials, e.g., one or more corrosion-resistant materials. Whatever the case, cathode interface separator 1701 may be formed in any suitable manner, such as additively manufactured, injection molded, compression molded, stamped, casted, machined, and/or the like.

### Anode Interface Assembly

FIG. 47 depicts an exploded view of an example anode interface assembly of the example multi-cell COₓ electrolyzer stack of FIG. 6. FIG. 48 depicts the example anode interface assembly of FIG. 47 in an assembled state. FIG. 44 depicts an example anode interface separator of FIG. 47.

As seen in at least FIGS. 5, 6, 11A, 44, 47, and 48, anode interface assembly 509 may include equivalent components as anode components 1101 of repeat unit 1100, except anode interface assembly 509 may omit third anode gaskets 1117c of second anode gasket set 1117 and include anode frame 4701 instead of anode frame 1115. As such, duplicative descriptions of equivalent components will be omitted to avoid obscuring embodiments disclosed herein. In addition, anode interface assembly 509 may include anode interface separator 4703, which may be configured substantially equivalent to separator plate 1107 of repeat unit 1100, except anode interface separator 4703 may exclude openings/orifices 4319-4335 (see FIG. 43). It is also noted that anode frame 4701 may be substantially equivalent to anode frame 1115 (see also FIGS. 37-42), except that anode frame 4701 may omit second fluidic inlet and outlet passages 3743 and 3745, recesses 4027 and 4029 in surface 3703, and first, second, and third fastener orifices 3761, 3763, and 3765, as well as swage nuts 1135. Thus, instead of anode frame 4701 being coupled to an adjacent cathode frame, such as cathode frame 1115, as in repeat unit 1100 described at least in association with FIG. 11A, anode frame 4701 may simply be interposed between unitized MEA assembly 1119_n of repeat unit 503_n and anode interface separator 4703 when anode interface assembly 509 is incorporated as part of stack 500 (see also FIGS. 5-10). As such, second and third anode gaskets 1113b and 1113c of first anode gasket set 1113 may interface with recesses in surface 4701a of anode frame 4701 similar to recesses 3749-3759 in surface 3701 of anode frame 1115 and abut against surface 2803 of cathode frame 1131 of repeat unit 503_n around first and second fluidic inlet and outlet passages 2815-2821 (see also FIGS. 28-36). Further, first anode gasket 1113a of first anode gasket set 1113 may interface with a recess in surface 4701a of anode frame 4701 similar to recess 3747 in surface 3701 of anode frame 1115, abut against a corresponding surface of support frame 1125 of unitized MEA assembly 1119 (see also FIGS. 25-27), and encircle opening 1125a in support frame 1125 (see also FIGS. 25-27). In a similar fashion, first and second anode gaskets 1117a and 1117b of second anode gasket set 1117 may simply interface with recesses in surface 4701b of anode frame 4701 similar to recesses 4017-4025 in surface 3703 of anode frame 1115 (see also FIGS. 39, 40, and 42) and may abut against first surface 4703a of anode interface separator 4703.

### Bladder

As previously discussed, bladder side assembly 511 (see, e.g., FIG. 5) may be at least configured to constrain axial expansion of the plurality of cells, such as cell 501, of stack 500 during the COₓ reduction process(es) in a manner that prevents or reduces the likelihood of the plurality of cells from being overly or insufficiently compressed, but maintain corresponding fluidic seals and electrical conductivity between associated components of stack 500. These features may be provided by the conjunction of bladder bus plate 521, insulation plate 523, end plate 525, gaskets 559 and 561, and fluidic inlet connector 563 (see, e.g., FIGS. 5-10).

FIG. 86 depicts a plan view of an illustrative insulation plate of the example multi-cell COₓ electrolyzer of FIG. 6. FIG. 87 depicts a cross-sectional view of the illustrative insulation plate of FIG. 86 taken along sectional line 87-87. FIG. 88 depicts a plan view of an illustrative end plate of the example multi-cell COₓ electrolyzer of FIG. 6. FIG. 89 depicts a cross-sectional view of the illustrative end plate of FIG. 88 taken along sectional line 89-89. FIG. 90 depicts an enlarged portion of the cross-sectional view of FIG. 9.

Referring to FIGS. 86 and 87, insulation plate 523 may be a generally rectangular plate-shaped body having first surface 8601 (e.g., a top surface) opposing second surface 8603 (e.g., a bottom surface) in axial direction 8605. Although insulation plate 523 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, insulation plate 523 will be described in association with a generally rectangular configuration. First and second surfaces 8601 and 8603 may be bounded by one or more peripheral surfaces, such as peripheral surfaces (or surfaces) 8607, 8609, 8611, and 8613 that may be connected to one another via one or more other peripheral surfaces, such as peripheral surface (or surface) 8615. In some embodiments, insulation plate 523 may have a symmetrical configuration about one or more reference planes perpendicular to axial direction 8605. For instance, a configuration of insulation plate 523 may be symmetrical about either or both of reference planes 8617 and 8619, but embodiments are not limited thereto.

According to various implementations, insulation plate 523 includes first recess 8621 in a central portion of surface 8601. First recess 8621 may not only terminate at surface 8623, but may also include extended portions 8625 and 8627 extending from a central area of first recess 8621 respectively towards peripheral surfaces 8609 and 8613. A size, shape, and location of first recess 8621 may be configured to enable at least a portion of bus plate 521 (see, e.g., FIGS. 5-10) to be received therein when stack 500 is assembled. As such, a corresponding portion of terminal portion 521t of bus plate 521 (see, e.g., FIGS. 5-10) may be received in one of extended portions 8625 and 8627. The central area of first recess 8621 may include second recess 8629 in a peripheral region thereof. Second recess 8629 may be configured to interface with gasket 559 (see, e.g., FIGS. 5 and 90) in a manner that, when bus plate 521 and insulation plate 523 are assembled as part of stack 500, lower surface 521b (see FIG. 90) of bus plate 521 may at least abut against gasket 559, and, depending on an extent of compression of the various components of stack 500, may either abut against surface 8623 of insulation plate 523 (such as shown in FIG. 90) or may be spaced apart from surface 8623 in an axial direction, which may extend parallel (or substantially parallel) to the z-axis direction shown in FIGS. 5 and 90 and may be the same as axial direction 8605. As will become more apparent below, a distance in axial direction 8605 between lower surface 521b of bus plate 521 and surface 8623 of insulation plate 523 may be controlled to constrain axial expansion of the plurality of cells, such as cell 501, of stack 500 (see, e.g., FIGS. 5-10) during the COₓ reduction process(es) to maintain corresponding fluidic seals and electrical conductivity between associated components of stack 500, but in a manner that prevents or reduces the likelihood that the plurality of cells (and the associated components of the cells) are overly compressed.

For example, one or more control fluids (e.g., gaseous COₓ) may be introduced between bus plate 521 and insulation plate 523 to regulate a distance between lower surface 521b of bus plate 521 and surface 8623 of insulation plate 523. In some embodiments, the one or more control fluids may be provided via orifice 8631 in surface 8623 that extends through insulation plate 523 to surface 8603. A size, shape, and location of orifice 8631 may correspond with a size, shape, and location of blind orifice 8801 in surface 525a of end plate 525 (see FIGS. 88-90). Blind orifice 8801 of end plate 525 may be fluidically connected to fluidic inlet connector 563 via fluidic passageway 8803 as seen in FIGS. 88-90. As such, the one or more control fluids may be caused to flow between bus plate 521 and insulation plate 523 via the conjunction of fluidic inlet connector 563, fluidic passageway 8803, blind orifice 8801, and orifice 8631, as well as source 9001 (see FIG. 90) of the one or more control fluids. In some embodiments, source 9001 of the one or more control fluids may be the same as the source of input providing, for instance, gaseous COₓ, to second fluidic inlet connector 547 (see FIG. 5). Regardless of the source, the distance between lower surface 521b of bus plate 521 and surface 8623 of insulation plate 523 may be controlled based on an accumulated pressure of the one or more control fluids in the area between lower surface 521b of bus plate 521 and surface 8623 of insulation plate 523, the area being peripherally bounded by gasket 559 (see also FIGS. 5 and 90). In this manner, regulating the distance between lower surface 521b of bus plate 521 and surface 8623 of insulation plate 523 may be utilized to constrain axial expansion of the plurality of cells, such as cell 501, during operation. This may help maintain corresponding fluidic seals and electrical conductivity between associated components of stack 500 (see, e.g., FIG. 5).

According to some embodiments, when the accumulated pressure in the area between lower surface 521b of bus plate 521 and surface 8623 of insulation plate 523 builds beyond a determined threshold, the distance between lower surface 521b of bus plate 521 and surface 8623 of insulation plate 523 may increase to point at which a fluidic seal formed between gasket 559 and lower surface 521b of bus plate 521 may become compromised. If and when the fluidic seal formed between gasket 559 and lower surface 521b of bus plate 521 becomes compromised, at least some of the one or more control fluids may escape (or bleed) from the area between lower surface 521b of bus plate 521 and surface 8623 of insulation plate 523 that may cause the accumulated pressure to decrease along with the distance between lower surface 521b of bus plate 521 and surface 8623 of insulation plate 523. In some embodiments, insulation plate 523 and/or end plate 525 may be configured with one or more fluidic passages interfacing with a relief valve configured to evacuate excess pressure built in the area between lower surface 521b of bus plate 521 and surface 8623 of insulation plate 523 to prevent over compression of the various components of stack 500 (see, e.g., FIG. 5).

In some embodiments, surface 525a (see FIG. 88) of end plate 525 may include recess 8805 encircling blind orifice 8801. Recess 8805 may be configured to interface with gasket 561 (see, e.g., FIGS. 5 and 90) such that, when insulation plate 523, end plate 525, gasket 565, and gasket 561 are incorporated as part of stack 500 (see, e.g., FIGS. 5 and 90), gasket 561 may not only be interposed between insulation plate 523 and end plate 525, but also form a fluidic seal between orifice 8631 in insulation plate 523 and blind orifice 8801 in end plate 525. The fluidic seal between orifice 8631 in insulation plate 523 and blind orifice 8801 in end plate 525 may be enhanced through the coupling of insulation plate 523 and end plate 525. As such, insulation plate 523 may include a plurality of fastener orifices 8633 (which may be countersunk with respect to surface 8601) to enable first fasteners 535 (see FIG. 5) to extend through insulation plate 523 and engage with corresponding fastener orifices 8807 (see FIG. 88) in end plate 525. Although only one set of mating orifices configured to enable the one or more control fluids to be flowed into the area between lower surface 521b of bus plate 521 and surface 8623 of insulation plate 523 are shown in FIGS. 86-90, insulation plate 523 and end plate 525 may be configured with more than one set of mating orifices. In some cases, a plurality of mating orifices may be provided and arranged about the central area of recess 8621 in insulation plate 523, such as arranged at regular (or substantially regular) rotation angles about, for instance, a reference axis coincident with axial direction 8605. Such a configuration may allow for a more uniform axial force to be exerted on bus plate 521 as pressure builds in the area between lower surface 521b of bus plate 521 and surface 8623 of insulation plate 523.

According to various embodiments, source 9001 may be configured to supply the gaseous COₓ to second fluidic inlet connector 547 (see, e.g., FIGS. 5-9) at a first pressure and to supply the one or more control fluids (e.g., gaseous COₓ) to fluidic inlet connector 563 (see, e.g., FIGS. 5-9 and 90) at a second pressure. In some embodiments, the first and second pressures may be equivalent or substantially equivalent. In some cases, source 9001 may be configured to control (e.g., adjust) one or more of the first and second pressures based on conditions of stack 500, e.g., based on an extent of expansion of the cells of stack 500 in the axial direction, based on an accumulated pressure in the area between lower surface 521b of bus plate 521 and surface 8623 of insulation plate 523, based on the temperature of one or more components of stack 500, and/or the like (see also FIGS. 5-10). As such, the first and second pressures may reach equilibrium, such as, in response to steady state conditions, e.g., steady state operational conditions of stack 500. It is also noted that source 9001 may be configured to supply the gaseous COₓ to second fluidic inlet connector 547 (see, e.g., FIGS. 5-9) at a first time and to supply the one or more control fluids (e.g., gaseous COₓ) to fluidic inlet connector 563 (see, e.g., FIGS. 5-9 and 90) at a second time. In some embodiments, the first and second times may occur simultaneously or substantially simultaneously. In some cases, source 9001 may be configured to delay the supply of the one or more control fluids to fluidic inlet connector 563 (see, e.g., FIGS. 5-9 and 90) with respect to the provisioning of the gaseous COₓ to second fluidic inlet connector 547 (see, e.g., FIGS. 5-9). For example, and with reference to FIGS. 5-9 and 90, source 9001 may be configured to delay the supply of the one or more control fluids to fluidic inlet connector 563 until one or more conditions are satisfied, e.g., an extent of expansion of one or more of the cells of stack 500 in the axial direction reaches one or more defined thresholds, a temperature of one or more components of stack 500 reaches one or more defined thresholds, flow of the gaseous COₓ to second fluidic inlet connector 547 reaches steady state condition(s), and/or the like.

With continued reference to FIGS. 86, 88, and 90, insulation plate 523 may include a plurality of datum openings 8635 configured to receive and support respective portions of datum rods 557 therein, and end plate 525 may further include fluidic inlet port 8809 configured to interface with fluidic inlet connector 563. Fluidic inlet port 8809 may include threaded region 8809t, which may be configured to engage with a respective threaded region of fluidic inlet connector 563. Alternatively, fluidic inlet connector 563 may be welded, e.g., sweat welded, to fluidic inlet port 8809 and threaded portion 8809t may be omitted.

### Anode Flow Fields

FIG. 83 depicts a plan view of a portion of an illustrative anode flow field of the example multi-cell COₓ electrolyzer of FIG. 6. FIGS. 84A and 84B depict respective cross-sectional views of the illustrative anode flow field of FIG. 83 taken along sectional lines 84A-84A and 84B-84B according to some embodiments.

With reference to FIGS. 11A, 83, 84A, and 84B, anode flow field 1111 may be a generally rectangular plate-shaped body including a plurality of projections 8301 protruding from surface 8303 of main body portion 8305 in the axial direction, which may extend parallel to the z-axis direction. In some embodiments, projections 8301 may be rectangular prisms having length 8307 in a first direction (e.g., the x-axis direction) transverse to the axial direction, width 8309 in a second direction (e.g., the y-axis direction) transverse to the axial direction and the first direction, and height 8311 in the axial direction, but embodiments are not limited thereto. For instance, one or more of projections 8301 may be alternatively formed as cylindrical prisms, triangular prisms, pentagonal prisms, and/or the like. Projections 8301 may be spaced apart from one another by pitch 8313 in the first direction and pitch 8315 in the second direction. Although projections 8301 are shown as being arranged in a plurality of parallel rows and parallel columns, embodiments are not limited thereto. For instance, adjacent rows and/or columns of projections 8301 may be offset from one another such as shown in FIG. 85A with respect to projections 8501. In some cases, pitches 8313 and 8315 may be equivalent (or substantially equivalent) to one another, but embodiments are not limited thereto. In this manner, fluidic passages 8317 may be formed between adjacent projections among projections 8301, and, thereby, form flow paths through which water (or other anolyte) may flow in a distributed manner generally from supply channels 3733 of anode frame 1115 to collection channels 3735 of anode frame 1115 (see FIG. 37-42) to provide water to anode PTL 1109, and, thereby, to the anode side of MEA 1105 (see FIG. 11A).

Although anode flow field 1111 has been described as having a generally rectangular plate-shaped body, any suitable geometric configuration may be utilized. For instance, anode flow field 1111 may have a generally circular, generally elliptical, generally triangular, generally pentagonal, generally hexagonal, etc., configuration. Whatever configuration is utilized, anode flow field 1111 should be able to be at least partially supported in opening 3723 (see, e.g., FIGS. 23, 24, and 37-42) in anode frame 1115. Further, although anode flow field 1111 has been described in association with a pin-type implementation, embodiments are not limited thereto. For instance, any other suitable anode flow field design may be utilized, such as parallel, serpentine, interdigitated, spiral, radial, etc. An example of a rotated pin-type embodiment will be described in more detail in association with FIGS. 85A-85C.

FIG. 85A depicts a plan view of a portion of an illustrative anode flow field of the example multi-cell COₓ electrolyzer of FIG. 6. FIGS. 85B and 85C depict respective cross-sectional views of the illustrative anode flow field of FIG. 85A taken along sectional lines 85B-85B and 85C-85C according to some embodiments.

With reference to FIGS. 11A and 85A-85C, anode flow field 1111 may be formed in a similar manner as described in association with FIGS. 83, 84A, and 84B, but the plurality of projections 8501 in FIGS. 85A-85C may be rotated by angle 8503 with respect to a first direction (e.g., the x-axis direction) to enable leading vertices 8501a of projections 8501 to split and distribute input anolyte flow 8505. In addition, adjacent rows and columns of projections 8501 may be offset from one another. For example, adjacent rows may be offset from one another by offset amount 8507 in the first direction transverse to the axial direction (e.g., the z-axis direction), and adjacent columns may be offset from one another by offset amount 8509 in a second direction (e.g., the y-axis direction) transverse to the axial direction and the first direction. In some cases, offset amounts 8507 and 8509 may be equivalent (or substantially equivalent) to one another, but embodiments are not limited thereto.

Similar to projections 8301 described in association with FIGS. 83, 84A, and 84B, projections 8501 may protrude from surface 8511 of main body portion 8513 in the axial direction, which may extend parallel (or substantially parallel) to the z-axis direction. As shown in FIGS. 85A-85C, projections 8501 may be diamond-shaped prisms having respective lengths 8515 in the first direction, corresponding widths 8517 in the second direction, and respective heights 8519 in the axial direction, but embodiments are not limited thereto. For instance, one or more of projections 8501 may be alternatively formed as elliptical prisms, oblong prisms, lenticular prisms, sinus prisms, and/or the like. Projections 8501 may be spaced apart from one another by pitch 8521 in the first direction and pitch 8523 in the second direction. In some cases, pitches 8521 and 8523 may be equivalent (or substantially equivalent) to one another, but embodiments are not limited thereto. In this manner, fluidic passages 8525 may be formed between adjacent projections among projections 8501, and, thereby, form flow paths through which water (or other anolyte) may flow in a distributed manner generally from supply channels 3733 of anode frame 1115 (see FIGS. 37-42) to collection channels 3735 of anode frame 1115 to provide water to anode PTL 1109 (see FIG. 11A), and, thereby, to the anode side of MEA 1105.

### Cathode Flow Fields

Various features and technologies may be used to help mitigate the detrimental effects of liquid water accumulation in COₓ electrolyzer cathodes. For example, the cathode flow field 1127 may be constructed so as to have one or more structural features that may allow for more effective liquid water management within the cell 501.

For example, both the anode flow field 1111 and the cathode flow field 1127 may have a corresponding anode channel(s) and cathode channel(s), respectively. The cathode channel(s) may, for example, be designed to have certain characteristics that may contribute to more effective water evacuation in the context of a COₓ electrolyzer and/or that may mitigate the potential performance degradation that may occur in such a COₓ electrolyzer in the event that liquid water collects within the cathode side of the cell 501.

### Serpentine Channel Flow Fields

While various geometries of flow field channels may be used in COₓ electrolyzers, multiple serpentine channels generally offer superior performance in terms of providing for reliable, even distribution of COₓ gas to the cathode GDL 1121, and thus the MEA 1105, while also facilitating reliable removal of liquid water that may otherwise accumulate within the cathode flow field 1127 and the cathode GDL 1121 (see FIG. 11A). A serpentine channel typically has repeated longer segments that extend in generally parallel directions and are fluidically connected together by shorter segments that are fluidically interposed between them in alternating fashion, much like a switchback.

For the purposes of this disclosure, the term "fluidically connected" is used with respect to volumes, plenums, holes, etc., that may be structurally connected with one another in some way in order to form a fluidic connection, similar to how the term "electrically connected" is used with respect to components that are connected together to form an electric connection. The term "fluidically interposed," if used, may be used to refer to a component, volume, plenum, or hole that is fluidically connected with at least two other components, volumes, plenums, or holes such that fluid flowing from one of those other components, volumes, plenums, or holes to the other or another of those components, volumes, plenums, or holes would first flow through the "fluidically interposed" component before reaching that other or another of those components, volumes, plenums, or holes. For example, if a pump is fluidically interposed between a reservoir and an outlet, fluid that flowed from the reservoir to the outlet would first flow through the pump before reaching the outlet.

Single serpentine channel arrangements may have limited water evacuation performance in the context of COₓ electrolyzers for larger-area cells (e.g., larger than 100 cm²). Nevertheless, their performance may be adequate for some applications. In a single serpentine channel arrangement, e.g., such as is shown in FIG. 49, a single, continuous serpentine channel 4956 switchbacks across an area 4952 of a cathode flow field 4916 bounded by shorter segments 4962 and first and last longer segments 4960. The serpentine channel 4956 is thus the only conduit for COₓ gas to enter a corresponding cathode GDL and MEA and is also the only conduit for liquid water that comes into the cathode flow field 4916 from the cathode GDL via that area. Thus, the rate at which liquid water is added to the serpentine channel 4956 is equal to the rate at which liquid water flows out of the area 4952 and into the cathode flow field 4916. The high rate of liquid water introduction into such a serpentine channel 4956, coupled with the long average distance that such water must travel in order to be pushed through the serpentine channel 4956 before reaching a fluidic outlet port, such as fluidic outlet port 4930, generally makes it very challenging to properly manage the liquid water levels within the cathode flow field 4916, rendering COₓ electrolyzers that use such single-channel serpentine cathode flow fields 4916 with significantly compromised performance compared to COₓ electrolyzers using, for example, multiple serpentine channel arrangements. In some implementations, a single serpentine channel has an overall channel length (distance from inlet to outlet) of about 12 m or less, or about 6 m or less, or about 2 m or less.

Multiple serpentine channels can refer to multiple separate serpentine channels that generally follow a common serpentine path, thereby resulting in an interleaved or nested arrangement of the separate serpentine channels, or can refer to multiple instances of the same serpentine channel (or nearly the same serpentine channel) that are arranged side-by-side or otherwise arranged so as to flow in parallel. FIG. 50 depicts the former arrangement, which may also be referred to herein as nested or interleaved multiple serpentine channel arrangements. In FIG. 50, four serpentine channels that generally follow the same serpentine path are shown (two are shown with interiors with white fill and two with interiors with shaded fill to make it easier to differentiate between them; a broken-line rectangle representing the combined open channel area and wall footprint area of a flow field having such an arrangement is also shown). The open channel area refers to the total area through which gas may exit the flow field and travel into the GDL; in a flow field with constant- and equal-width paths, the open channel area would generally be equal to the total path length of the channel(s) times the channel width. The wall footprint area of a flow field refers to the area of the portion of the flow field that defines walls between adjacent portions of a channel or channels of the flow field and that is pressed into contact with the GDL. Thus, both areas are evaluated within the plane of the flow field that is pressed into contact with the GDL. Fluid may be introduced into/removed from the serpentine channels through the inlet and outlet ports (the short segments terminating in small solid black circles). In FIG. 51, a similar arrangement is shown for a side-by-side arrangement of four multiple serpentine channels, which may also be referred to herein as side-by-side multiple serpentine channels. A similar convention with regard to the inlet/outlet, combined open channel area and wall footprint area, and use of shaded/unshaded fill to illustrate the different channels is used in FIG. 51 as in FIG. 50.

In such arrangements, the total length of each individual serpentine channel may generally be equal to the total lengths of the other individual serpentine channels in the multiple serpentine channels (although in the nested or interleaved multiple serpentine channel arrangements, some small variation in length may be present depending on how the channels are arranged, e.g., whether or not there is an odd or even number of longer segments in each channel), resulting in generally equal flow resistance, pressure drop, and transit time between the channels (assuming that each such channel is fluidically connected with the same fluidic environments on both ends).

FIG. 52 depicts an example of a cathode flow field 5216 that includes a two-channel multiple serpentine channel arrangement. As can be seen, the cathode flow field 5216 has a fluidic inlet port 5228 and a fluidic outlet port 5230. Two serpentine channels 5256a and 5256b are shown which follow a common serpentine path (not shown, but would generally be represented by the path followed by partition wall 5266, which separates the two serpentine channels 5256a and 5256b). The serpentine channels 5256a and 5256b switchback across an area 5252 in a generally tandem fashion. As a result, fluid that is flowed through either of the serpentine channels 5256a and 5256b, e.g., COₓ gas, may generally be evenly delivered to an adjoining cathode GDL within a region corresponding to the area 5252. At the same time, any liquid water that is flowed into the cathode flow field 5216 from the adjoining cathode GDL may correspondingly tend to be evenly delivered to both serpentine channels 5256a and 5256b. Thus, each serpentine channel 5256 would receive, assuming that the cathode flow field 5216 is substituted for the cathode flow field 4916 of FIG. 49, approximately half the water that was delivered to the single serpentine channel 4956 of FIG. 49. Generally speaking, the amount of water delivered to each serpentine channel in a cathode flow field having a multiple serpentine channel arrangement will be equivalent to the total amount of water received by the multiple serpentine channel arrangement divided by the number of separate channels in the multiple serpentine channel arrangement. This has the effect of reducing the amount of water that must be evacuated from each serpentine channel per unit time, which may make it more feasible to properly manage the liquid water conditions within a COₓ electrolyzer if the gas flow velocity is maintained or at least not proportionately decreased. For example, the lower per channel quantities of water will have less mass and require less energy in order to be pushed through the channels to the fluidic outlet port 5230 of the cathode flow field 5216. As a result, lower pressure differentials between the fluidic inlet port 5228 and fluidic outlet port 5230 of the cathode flow field 5216 may be used while still providing for efficient evacuation of liquid water from the cathode flow field 5216.

Multiple serpentine channels may also allow for relatively even distribution of the fluid that flows within them across the cathode GDL 1121 but with decreased total flow path length for each such serpentine channel as compared with multiple serpentine channel or single serpentine channel implementations having the same or similar channel depth and width and total open channel area in contact with the cathode GDL 1121 but with fewer numbers of such channels. For example, for a given multiple serpentine channel arrangement, it may be desirable to maintain the distance between adjacent portions of at least the longer portions of the serpentine channel(s) to be within a minimum distance of each other. For each additional serpentine channel that is included in a multiple serpentine channel arrangement, meeting such inter-channel spacing restrictions may be attained using serpentine channels of increasingly shorter overall lengths. For clarity, the overall length of a serpentine channel refers to the total of the average path lengths for all of the longer segments of the serpentine channel plus the total average path length of shorter segments that fluidically connect those longer segments with one another, plus the total average path length of any other segments that are fluidically interposed between the inlet and outlet of the serpentine channel.

Moreover, as serpentine channels decrease in length, the average potential distance that liquid water must travel in order to be expelled from such a serpentine channel will also decrease, as does generally the maximum amount of water that would potentially need to be removed. As a result, less energy is required to evacuate water from such serpentine channels in the event that water collects within such a serpentine channel; this is because the maximum amount of water that may need to be removed from such a channel will be less than in longer-length channels (of the same general cross-sectional area)-there is thus less mass to move. Moreover, the distance that such a water mass must be displaced by in order to push it through such a channel to the fluidic outlet port will generally be less than the distance that a similar water mass must be displaced by in order to be pushed through a longer-length channel to the fluidic outlet port. Of course, the distance that the water mass must be displaced by in order to be pushed through the channel to the fluidic outlet port is dependent on where the water mass is located within the channel. However, on average, water masses that collect in shorter-length channels will generally need to be displaced by a lesser amount than water masses that collect in longer-length channels in order to move such water masses to the fluidic outlet port of the flow field having such channels. Since less energy is needed to move such water masses (droplets) in flow fields with shorter-length passages, lower gas flow velocities, and lower pressure drops, may be used. In some embodiments, a cathode flow field has a serpentine channel with a length of about 12 m or less, or about 10 m or less, or about 6 m or less. For example, serpentine channels that have overall lengths on the order of less than about 6 meters, e.g., less than about 6 meters, less than about 5.5 meters, less than about 5 meters, less than about 4.5 meters, less than about 4 meters, less 3.5 meters, less than about 3 meters, less than about 2.5 meters, or less than about 2 meters may, in some implementations, provide a fluid flow path in the cathode flow field 1127 that allows for the flow of COₓ gas to be distributed across a wide area of the cathode GDL 1121 while, at the same time, avoiding being so long that evacuating liquid water from within such serpentine channels becomes too difficult. At the same time, serpentine channels that are too short may make it challenging to maintain a desired pressure drop (see later discussion below) across the cathode flow field 1127. To that end, some cathode flow field serpentine channels may be configured to also have overall lengths greater than or equal to 1.5 meters.

**In** some implementations, the length of an individual serpentine channel for a cathode flow field may be between about 1.5 m and about 12 m, between about 1.5 m and about 6 m, between about 1.5 m and about 3.8 m, between about 3.8 m and about 6 m, between about 1.5 m and about 2.6 m, between about 2.6 m and about 3.8 m, between about 3.8 m and about 4.9 m, between about 4.9 m and about 6 m, between about 1.5 m and about 2.1 m, between about 2.1 m and about 2.6 m, between about 2.6 m and about 3.2 m, between about 3.2 m and about 3.8 m, between about 3.8 m and about 4.3 m, between about 4.3 m and about 4.9 m, between about 4.9 m and about 5.4 m, between about 5.4 m and about 6 m, between about 1.5 m and about 1.8 m, between about 1.8 m and about 2.1 m, between about 2.1 m and about 2.3 m, between about 2.3 m and about 2.6 m, between about 2.6 m and about 2.9 m, between about 2.9 m and about 3.2 m, between about 3.2 m and about 3.5 m, between about 3.5 m and about 3.8 m, between about 3.8 m and about 4 m, between about 4 m and about 4.3 m, between about 4.3 m and about 4.6 m, between about 4.6 m and about 4.9 m, or between about 4.9 m and about 5.2 m. It will be understood that reference herein, both above and below, to a value being "between" two other values, unless the context indicates otherwise, is inclusive of the values in between the two other values as well as the values themselves.

**In** cathode flow fields with serpentine channels, it may be beneficial to configure the serpentine channels to have particular structural characteristics that may provide for enhanced liquid water removal while at the same time providing for effective COₓ delivery to the cathode GDL. For example, serpentine channels within the length ranges discussed above may be further constrained to have particular widths (the dimension of a serpentine channel in a direction parallel to the plane of the cathode GDL 1121 and transverse to the path that the channel follows (or, generally, transverse to the nominal flow direction of fluid flow through the channel)) and depths (the dimension of a serpentine channel in a direction perpendicular to the plane of the cathode GDL 1121) to further enhance their water-removal performance in the context of a COₓ electrolyzer. For clarity, the cathode GDL 1121 is generally in the form of a thin sheet that, when stacked with the MEA 1105 (see, e.g., FIG. 11A) and the anode PTL 1109 (see, e.g., FIG. 11A), is compressed between the cathode flow field 1127 and the anode flow field 1111 into a nominally planar geometry; reference to "the plane of the cathode GDL" is thus to be understood to refer to a plane that is generally parallel to, and coincident with, the cathode GDL 1121 in such a state. For example, such serpentine channels may have widths that are between about 0.3 mm and about 2 mm, between about 0.3 mm and about 1.2 mm, between about 1.2 mm and about 2 mm, between about 0.3 mm and about 0.72 mm, between about 0.72 mm and about 1.2 mm, between about 1.2 mm and about 1.6 mm, between about 1.6 mm and about 2 mm, between about 0.3 mm and about 0.51 mm, between about 0.51 mm and about 0.72 mm, between about 0.72 mm and about 0.94 mm, between about 0.94 mm and about 1.2 mm, between about 1.2 mm and about 1.4 mm, between about 1.4 mm and about 1.6 mm, between about 1.6 mm and about 1.8 mm, or between about 1.8 mm and about 2 mm.

Such serpentine channels may also have depths that are between about 0.3 mm and about 3 mm, between about 0.3 mm and about 1.6 mm, between about 1.6 mm and about 3 mm, between about 0.3 mm and about 0.98 mm, between about 0.98 mm and about 1.6 mm, between about 1.6 mm and about 2.3 mm, between about 2.3 mm and about 3 mm, between about 0.3 mm and about 0.64 mm, between about 0.64 mm and about 0.98 mm, between about 0.98 mm and about 1.3 mm, between about 1.3 mm and about 1.6 mm, between about 1.6 mm and about 2 mm, between about 2 mm and about 2.3 mm, between about 2.3 mm and about 2.7 mm, or between about 2.7 mm and about 3 mm.

In particular, in some cathode flow field implementations with serpentine channels, the channels may be dimensioned such that the open surface area per channel, i.e., the area that is bounded by the edges of the channel that contact the cathode GDL, is between about 750 mm² and about 200,000 mm², between about 750 mm² and about 100,000 mm², between about 100,000 mm² and about 200,000 mm², between about 750 mm² and about 51,000 mm², between about 51,000 mm² and about 100,000 mm², between about 100,000 mm² and about 150,000 mm², between about 150,000 mm² and about 200,000 mm², between about 750 mm² and about 26,000 mm², between about 26,000 mm² and about 51,000 mm², between about 51,000 mm² and about 75,000 mm², between about 75,000 mm² and about 100,000 mm², between about 100,000 mm² and about 130,000 mm², between about 130,000 mm² and about 150,000 mm², between about 150,000 mm² and about 180,000 mm², or between about 180,000 mm² and about 200,000 mm².

**In** some such implementations, such channels may be further dimensioned such that the cross-sectional area (or areas, if the channel has a varying cross-sectional area along its length) of each such channel, i.e., the area of the channel in a plane that is perpendicular to the direction of flow of fluid through the channel under normal operating conditions or to the path that the channel follows across the cathode flow field, is between about 0.15 mm² and about 6 mm², between about 0.15 mm² and about 3.1 mm², between about 3.1 mm² and about 6 mm², between about 0.15 mm² and about 1.6 mm², between about 1.6 mm² and about 3.1 mm², between about 3.1 mm² and about 4.5 mm², between about 4.5 mm² and about 6 mm², between about 0.15 mm² and about 0.88 mm², between about 0.88 mm² and about 1.6 mm², between about 1.6 mm² and about 2.3 mm², between about 2.3 mm² and about 3.1 mm², between about 3.1 mm² and about 3.8 mm², between about 3.8 mm² and about 4.5 mm², between about 4.5 mm² and about 5.3 mm², or between about 5.3 mm² and about 6 mm².

In yet further implementations, the total channel volume of each such channel may be between about 200 µl and about 36,000 µl, between about 200 µl and about 18,000 µl, between about 18,000 µl and about 36,000 µl, between about 200 µl and about 9,200 µl, between about 9,200 µl and about 18,000 µl, between about 18,000 µl and about 27,000 µl, between about 27,000 µl and about 36,000 µl, between about 200 µl and about 4,700 µl, between about 4,700 µl and about 9,200 µl, between about 9,200 µl and about 14,000 µl, between about 14,000 µl and about 18,000 µl, between about 18,000 µl and about 23,000 µl, between about 23,000 µl and about 27,000 µl, between about 27,000 µl and about 32,000 µl, or between about 32,000 µl and about 36,000 µl.

In some such implementations, cathode flow fields with serpentine channels may also have structural characteristics relating to the thickness of the walls that are interposed between adjacent longer segments of one or more of the serpentine channels. For example, the wall thickness in between adjacent longer segments of one or more of the serpentine channels (and thus the distance between surfaces of that channel or those channels that are closest to one another) may be selected to be between about between about 0.00005 and about 0.0013333, between about 0.00005 and about 0.00069, between about 0.00069 and about 0.0013333, between about 0.00005 and about 0.00037, between about 0.00037 and about 0.00069, between about 0.00069 and about 0.001, between about 0.001 and about 0.0013333, between about 0.00005 and about 0.00021, between about 0.00021 and about 0.00037, between about 0.00037 and about 0.00053, between about 0.00053 and about 0.00069, between about 0.00069 and about 0.00085, between about 0.00085 and about 0.001, between about 0.001 and about 0.0012, or between about 0.0012 and about 0.0013333 times the average overall length of that serpentine channel or those serpentine channels (the latter case applying if the wall separates the longer portions of two different serpentine channels from each other-for clarity, in this instance the "average" overall length is half the sum of the overall lengths of both serpentine channels). In some such serpentine channel implementations having dimensional characteristics like those discussed above, the wall thickness may be, for example, between about 0.3 mm and about 2 mm, between about 0.3 mm and about 1.2 mm, between about 1.2 mm and about 2 mm, between about 0.3 mm and about 0.72 mm, between about 0.72 mm and about 1.2 mm, between about 1.2 mm and about 1.6 mm, between about 1.6 mm and about 2 mm, between about 0.3 mm and about 0.51 mm, between about 0.51 mm and about 0.72 mm, between about 0.72 mm and about 0.94 mm, between about 0.94 mm and about 1.2 mm, between about 1.2 mm and about 1.4 mm, between about 1.4 mm and about 1.6 mm, between about 1.6 mm and about 1.8 mm, or between about 1.8 mm and about 2 mm.

Serpentine channel cathode flow fields having characteristics such as those discussed above may offer superior liquid water evacuation performance in the context of COₓ electrolyzers, e.g., under operating conditions typically seen in COₓ electrolyzers (such as are discussed earlier herein) as compared with serpentine channel cathode flow fields having other such characteristics, such as may be designed for use with fuel cells.

While including increasingly higher numbers of multiple serpentine channels in a cathode flow field would generally seem desirable, unfettered increases in the number of flow field channels of the cathode flow field 1127 may be counterproductive. Each additional parallel flow field channel that exists in the cathode flow field 1127 may represent another path that fluid flowing through the multiple serpentine channels may take if blocked from flowing through one or more other serpentine channels in the arrangement of multiple serpentine channels. When such a rerouting of fluid occurs, it may cause an increase in the pressure differential along the channel, e.g., from channel start to channel end, that may cause the fluid that is pressing against the blockage to apply greater pressure on the blockage, thereby increasing the likelihood that the blockage (liquid water) will be dislodged, propelled through the serpentine channel that is being blocked, and eventually evacuated from the cathode flow field 1127 via flow field outlet such as flow field outlet 5930. However, if there are a sufficiently high enough number of channels present, the blockage of any one of them (or a small number of them) may result in a much smaller increase in the pressure differential in any single channel that may occur when an equivalent number of channels is blocked in a flow field with a lesser number of channels. In short, the gas flow that is blocked and reroutes through the other unblocked channels may be divided among a larger number of alternate channels, thereby resulting in a smaller amount of extra gas that must flow through each unblocked channel than might be the case with a lower number of channels in a similar blockage situation. The smaller the amount of extra gas that must flow through each channel during a blockage situation, the smaller the change in pressure drop that is needed to accommodate such a change. As a result, the increase in pressure drop that may occur in unblocked channels when gas flows re-route therethrough due to a blocked channel or channels decreases as the number of channels that are present increases.

At the same time, if the total lengths of the serpentine passages are sufficiently long, e.g., 0.3 m to 6 m, the pressure drop that occurs across each such channel may be high enough that it may act to help dislodge any obstructions, e.g., water, that may exist within any individual serpentine channel regardless of the number of channels present. For example, serpentine channels for COₓ electrolyzers may have dimensions and operational conditions, e.g., fluidic inlet port pressures, that are selected so as to produce a 0.001 psi to 4 psi pressure drop during normal operational flows for such serpentine channels, which may be high enough to dislodge potential water blockages that may be present within the serpentine channels; while higher pressure drops may be used as well, they may be unnecessary with respect to water evacuation and simply result in wasted energy that is needed to move the fluids through the serpentine channels under such pressure drop conditions. In some implementations, serpentine channels for COₓ electrolyzers may have dimensions and operational conditions, e.g., fluidic inlet port pressures, that are selected so as to produce, during normal operational flow conditions for a COₓ electrolyzer, a pressure drop of between about 0.001 psi and about 4 psi, between about 0.001 psi and about 2 psi, between about 2 psi and about 4 psi, between about 0.001 psi and about 1 psi, between about 1 psi and about 2 psi, between about 2 psi and about 3 psi, between about 3 psi and about 4 psi, between about 0.001 psi and about 0.5 psi, between about 0.5 psi and about 1 psi, between about 1 psi and about 1.5 psi, between about 1.5 psi and about 2 psi, between about 2 psi and about 2.5 psi, between about 2.5 psi and about 3 psi, between about 3 psi and about 3.5 psi, between about 3.5 psi and about 4 psi, between about 0.001 psi and about 0.25 psi, between about 0.25 psi and about 0.5 psi, between about 0.5 psi and about 0.75 psi, between about 0.75 psi and about 1 psi, between about 1 psi and about 1.3 psi, between about 1.3 psi and about 1.5 psi, between about 1.5 psi and about 1.8 psi, between about 1.8 psi and about 2 psi, between about 2 psi and about 2.3 psi, between about 2.3 psi and about 2.5 psi, between about 2.5 psi and about 2.8 psi, between about 2.8 psi and about 3 psi, between about 3 psi and about 3.3 psi, between about 3.3 psi and about 3.5 psi, between about 3.5 psi and about 3.8 psi, between about 3.8 psi and about 4 psi, between about 0.001 psi and about 0.13 psi, between about 0.13 psi and about 0.25 psi, between about 0.25 psi and about 0.38 psi, between about 0.38 psi and about 0.5 psi, between about 0.5 psi and about 0.63 psi, between about 0.63 psi and about 0.75 psi, between about 0.75 psi and about 0.88 psi, between about 0.88 psi and about 1 psi, between about 1 psi and about 1.1 psi, between about 1.1 psi and about 1.3 psi, between about 1.3 psi and about 1.4 psi, between about 1.4 psi and about 1.5 psi, between about 1.5 psi and about 1.6 psi, between about 1.6 psi and about 1.8 psi, between about 1.8 psi and about 1.9 psi, between about 1.9 psi and about 2 psi, between about 2 psi and about 2.1 psi, between about 2.1 psi and about 2.3 psi, between about 2.3 psi and about 2.4 psi, between about 2.4 psi and about 2.5 psi, between about 2.5 psi and about 2.6 psi, between about 2.6 psi and about 2.8 psi, between about 2.8 psi and about 2.9 psi, between about 2.9 psi and about 3 psi, between about 3 psi and about 3.1 psi, between about 3.1 psi and about 3.3 psi, between about 3.3 psi and about 3.4 psi, between about 3.4 psi and about 3.5 psi, between about 3.5 psi and about 3.6 psi, between about 3.6 psi and about 3.8 psi, between about 3.8 psi and about 3.9 psi, or between about 3.9 psi and about 4 psi. In some other implementations, serpentine channels for COₓ electrolyzers may have dimensions and operational conditions, e.g., fluidic inlet port pressures, that are selected so as to produce, during normal operational flow conditions for a COₓ electrolyzer, a pressure drop of between about 4 psi and about 50 psi, between about 4 psi and about 27 psi, between about 27 psi and about 50 psi, between about 4 psi and about 16 psi, between about 16 psi and about 27 psi, between about 27 psi and about 38 psi, between about 38 psi and about 50 psi, between about 4 psi and about 9.8 psi, between about 9.8 psi and about 16 psi, between about 16 psi and about 21 psi, between about 21 psi and about 27 psi, between about 27 psi and about 33 psi, between about 33 psi and about 38 psi, between about 38 psi and about 44 psi, between about 44 psi and about 50 psi, between about 4 psi and about 6.9 psi, between about 6.9 psi and about 9.8 psi, between about 9.8 psi and about 13 psi, between about 13 psi and about 16 psi, between about 16 psi and about 18 psi, between about 18 psi and about 21 psi, between about 21 psi and about 24 psi, between about 24 psi and about 27 psi, between about 27 psi and about 30 psi, between about 30 psi and about 33 psi, between about 33 psi and about 36 psi, between about 36 psi and about 38 psi, between about 38 psi and about 41 psi, between about 41 psi and about 44 psi, between about 44 psi and about 47 psi, or between about 47 psi and about 50 psi. In some other implementations, serpentine channels for COₓ electrolyzers may have dimensions and operational conditions, e.g., fluidic inlet port pressures, that are selected so as to produce, during normal operational flow conditions for a COₓ electrolyzer, a pressure drop of between about 0.001 psi and about 50 psi, between about 0.001 psi and about 25 psi, between about 25 psi and about 50 psi, between about 0.001 psi and about 13 psi, between about 13 psi and about 25 psi, between about 25 psi and about 38 psi, between about 38 psi and about 50 psi, between about 0.001 psi and about 6.3 psi, between about 6.3 psi and about 13 psi, between about 13 psi and about 19 psi, between about 19 psi and about 25 psi, between about 25 psi and about 31 psi, between about 31 psi and about 38 psi, between about 38 psi and about 44 psi, or between about 44 psi and about 50 psi. Pressure drops in the ranges listed above may be high enough to dislodge potential water blockages that may be present within such serpentine channels, particularly in the context of the higher water generation rates that COₓ electrolyzers tend to exhibit.

FIGS. 53 through 55 depict an example cathode flow field 5316 that may be used in some implementations. The depicted flow field has 15 channels and 9 passes. In one implementation, the depicted flow field has a planar surface area (facing a GDL) of 700 cm². FIG. 53 depicts an isometric view of the cathode flow field 5316. FIG. 55 depicts a detail view of the portion of FIG. 53 enclosed by a circle. FIG. 54 depicts the isometric view of FIG. 53, but with most of the channels of the flow field omitted, leaving only three channels 5358a, 5358b, and 5358c visible; this view is intended to make it easier to see the representative serpentine paths followed by the various channels. The cathode flow field 5316 actually includes 15 channels 5358. The channels in the example cathode flow field 5316 are each 0.66 mm deep by 0.81 mm wide, and each have a length of about 2,310 mm, a channel open area of about 1,880 mm², and a volume of about 1,240 mm³. The total open channel area of the cathode flow field 5316 is, in this example, 28,200 mm². With each of the 15 channels being separated from any adjacent channels by walls of 1.12 mm in width and the cathode flow field having dimensions of about 265 mm by 265 mm, about 40% of the cathode flow field 5316 surface area is taken up by the channels 5358. The depicted cathode flow field 5316 is designed to receive (and deliver) fluids from external manifolds that may be mounted against the external edges of the cathode flow field 5316 so as to flow fluid into or out of the channels 5358 from the side.

FIGS. 56 through 58 depict another example cathode flow field 5616 that may be used in some implementations. The depicted flow field has 34 channels and 7 passes. In one implementation, the depicted flow field has a planar surface area (facing a GDL) of 1,600 cm². As with FIGS. 53 through 55, FIG. 56 depicts an isometric view of the cathode flow field 5616 and FIG. 58 depicts a detail view of the portion of FIG. 56 enclosed by a circle. FIG. 57 depicts the isometric view of FIG. 56, but with most of the channels of the flow field omitted, leaving only three channels 5658a, 5658b, and 5658c visible; as with FIG. 55, this view is intended to make it easier to see the representative serpentine paths followed by the various channels. The cathode flow field 5616 actually includes 34 channels 5658. The channels in the example cathode flow field 5616 are each 0.66 mm deep by 0.76 mm wide, and each have a length of about 2,440 mm, a channel open area of about 1,880 mm², and a volume of about 1,230 mm³. The total open channel area of the cathode flow field 5616 is, in this example, 63,230 mm². With each of the 34 channels being separated from any adjacent channels by walls of 1.14 mm in width and the cathode flow field 5616 having dimensions of about 360 mm by 450 mm, about 39% of the cathode flow field 5616 surface area is taken up by the channels 5658. As with the cathode flow field 5316, the depicted cathode flow field 5616 is designed to receive (and deliver) fluids from external manifolds that may be mounted against the external edges of the cathode flow field so as to flow fluid into or out of the channels 5658 from the side.

In certain embodiments, a serpentine flow field as in FIGS. 53-58, the channel depth is about 0.5 mm to 1.5 mm. In certain embodiments, the nominal length of each flow channel in a flow field of FIGS. 53-58 is about 300 mm to 3,000 mm. In certain embodiments, the nominal channel width in a flow field of FIGS. 53-58 is about 0.5 mm to 1 mm. In certain embodiments, the nominal channel separation distance in a flow field of FIGS. 53-58 is about 1 mm to 1.5 mm.

In some implementations, serpentine channel cathode flow fields may feature serpentine channels that have rounded or smooth transitions between the longer and shorter segments as opposed to sharp transitions between such segments. For example, FIG. 59 depicts an example of a cathode flow field 5916 that has four cathode serpentine channels 5956 arranged in a multiple serpentine channel arrangement. It will be noted that unlike the single-channel and two-channel serpentine arrangements depicted in FIGS. 49 and 52, the transitions between the longer segments are provided by arcuate shorter segments instead of straight shorter segments. In other implementations, the shorter segments may still include a straight portion but may be joined to fluidically adjacent longer segments by smaller arcuate segments. Such cathode flow fields may further enhance the water evacuation performance of a COₓ electrolyzer since the absence of sharp interior corners in the serpentine channels may eliminate a potential dead zone or stagnation location for fluid flow that could otherwise serve as a location where liquid water could collect and reside indefinitely during use of the cathode flow field.

Other aspects of flow field channels may be alternatively or additionally modified as well in order to promote more effective liquid water evacuation. FIG. 60, for example, depicts a cross-sectional view of a cathode flow field 6016 that is pressed against a cathode GDL 6014. A plurality of square- or rectangular-cross-section serpentine channels 6056 are formed in the face of the cathode flow field 6016 that is pressed against the cathode GDL 6014. These serpentine channels 6056 have sharp corners at their interior bottom edges 6057, which may act to create small fluid flow stagnation areas that may prevent liquid water from being readily evacuated during normal COₓ electrolyzer operating conditions.

FIG. 61, by contrast, shows a cross-sectional view of a similar structure with a cathode flow field 6116 that is pressed against a cathode GDL 6114. A plurality of square- or rectangular-cross-section serpentine channels 6156 are formed in the face of the cathode flow field 6116 that is pressed against the cathode GDL 6114. Unlike the serpentine channels 6056, the serpentine channels 6156 have rounded corners at their interior bottom edges 6157, which may act to reduce flow stagnation in the bottom interior edge regions of such channels, thereby promoting liquid water evacuation during normal COₓ electrolyzer operating conditions.

FIG. 62 is a further example of a cathode flow field that may more readily evacuate liquid water during normal COₓ electrolyzer operating conditions. As can be seen, a cathode flow field 6216 is pressed against a cathode GDL 6214. A plurality of U-shaped cross-section serpentine channels 6256 are formed in the face of the cathode flow field 6216 that is pressed against the cathode GDL 6214. In this case, there effectively are no interior bottom edges of the serpentine channels 6256 since the bottom surface of such serpentine channels 6256 is semicircular, which may act to further reduce flow stagnation in such channels, thereby further promoting liquid water evacuation during normal COₓ electrolyzer operating conditions.

In some other or additional implementations, serpentine channel cathode flow fields may have variable-width walls in between some or all of the longer segments of one or more serpentine channels. FIG. 63 depicts an example of such a cathode flow field. In FIG. 63, a cathode flow field 6316 is shown which has a four-channel serpentine arrangement with each serpentine channel 6356 having longer segments 6360 and shorter segments 6362. It will be noted that the multiple serpentine channel arrangement has "peninsular" walls 6364 that are interposed between neighboring longer segments 6360 of a common serpentine channel 6356a (or 6356b) that have opposing fluid flow directions when fluid is flowing through the serpentine channels 6356 (generally all nested or interleaved multiple serpentine channel arrangements will have peninsular walls; they are only specifically called out here due to the particulars of this example implementation).

As can be seen in FIG. 63, the peninsular walls 6364 may have a varying wall thickness. For example, the peninsular walls 6364 have a root width 6368 where the peninsular walls 6364 "connect" with the outer perimeter region of the cathode flow field 6316 (which may be thought of as the "root" of the peninsular wall) and a tip width 6370 at their opposite ends. The increased width at the root as compared with the tip of the peninsular walls 6364 may reduce the chance of gas flow through the cathode GDL that might bypass some or all of the longer segments 6360 that are separated by the peninsular walls 6364 by passing under the wall, i.e., through the GDL that is sandwiched between the cathode flow field 6316 and the MEA (not shown, but see FIG. 11A) and which, in effect, caps the cathode serpentine channels 6356.

For example, in a serpentine channel of a cathode flow field that has portions thereof that are adjacent to one another, e.g., the outermost or innermost serpentine channel on a multi-channel, interleaved serpentine channel arrangement, gas that is flowed through such a channel, e.g., from point A to point B may experience a pressure drop/flow resistance if travelling from point A to point B via flow through point C that may, under some circumstances, exceed the pressure drop/flow resistance that may be experienced by that gas if it simply flowed from point A to point B more directly, e.g., by passing under the peninsular wall 6364 in between points A and B by way of the porous GDL that spans between points A and B and under the peninsular wall 6364. For example, if water accumulates in the channel between points A and C and/or between points C and B, the resulting blockage may increase the pressure drop/flow resistance for gas that flows along this path that it exceeds the pressure drop/flow resistance that the gas would experience if traveling from point A to point B more directly, e.g., under the peninsular wall 6364. As the flow path between points A and B under the peninsular wall 6364 may offer less flow resistance than the flow path between A and B via point C, the gas may then preferentially flow from point A under the peninsular wall 6364 to point B rather than via point C, thus depriving the GDL and MEA of exposure to gas that would normally flow through point C, thereby decreasing the efficiency of the COₓ cell in which the cathode flow field 6316 is used. To prevent this from happening, or to at least reduce the chances of this occurring, in some implementations, the peninsular walls 6364 may simply have a constant thickness along their lengths but may be thicker than partition walls 6366 that may separate other neighboring longer segments 6360 that have fluid flows in the same directions, thereby increasing the flow resistance experienced by gas that attempts to flow under the peninsular walls 6364. In other implementations, such as that shown in FIG. 63, the peninsular walls 6364 may taper towards their tips such that the tip width 6370 is less than the root width 6368, thereby causing the flow resistance under the peninsular walls 6364 to decrease from what it was near the root of a peninsular wall 6364 as the flow nears the tip of the peninsular wall 6364. This may assist with discouraging the flow of gas under the peninsular walls 6364 near the roots of those walls, but this effect may also decrease as the gas flow moves along the peninsular wall 6364 towards the tip thereof-however, the flow resistance along the desired flow path (via point C, for example) may also decrease, and there may thus not be as much of an incentive for gas to flow under the peninsular walls near the tips of the peninsular walls 6364. By tapering the thickness of the peninsular walls, the area of the cathode GDL that is compressed under the peninsular walls 6364 may be reduced as compared with non-tapering peninsular walls 6364, thereby increasing the area of the cathode GDL which has direct exposure to gas flow through the channels and increasing the opportunity for a reduction reaction to occur with such gas.

### Mirror Serpentine Channel Flow Fields

In the serpentine channel flow fields discussed above, the serpentine channels discussed generally do not exhibit any mirroring or bilateral symmetry. A further class of serpentine channel flow fields may, however, feature serpentine channels that are arranged in a generally bilaterally symmetric manner. In such flow fields, the flow field may generally be partitioned into two zones. The two zones may be generally equally sized and shaped, and may each contain a similar number of serpentine channels. The serpentine channel or channels in each zone may be arranged so as to generally be mirror images of one another with respect to the boundary between the two zones, e.g., the serpentine channels may exhibit bilateral symmetry about the boundary between the two zones.

FIG. 64 depicts a plan view of a simplified representation of an example mirror image cathode flow field. In FIG. 64, a cathode flow field 6416 is shown that is partitioned into two zones 6470 that are generally the same shape and size. A boundary 6472 is defined in between the two zones 6470; the zones 6470 are generally symmetrically arranged on either side of the boundary 6472. Each zone 6470 in this example includes a single cathode serpentine channel 6456, although it will be understood that each zone may include a larger number of cathode serpentine channels 6456 that follow a common path in a nested or interleaved manner, as with examples discussed earlier. The cathode serpentine channels 6456 each extend between a corresponding fluidic inlet port 6428 and a corresponding fluidic outlet port 6430 (it will be understood that these fluidic inlet ports 6428 may, for example, terminate in the same location, e.g., a common flow passage or manifold, and that the fluidic outlet ports 6430 may be similarly configured).

As is discussed further below, the symmetric arrangement of the cathode serpentine channels 6456 may provide various advantages over non-symmetric arrangements of cathode serpentine channels with respect to maintaining flow uniformity across the cathode flow field 6416. For example, the two zones 6470 may, together, generally represent an active area of the cathode flow field 6416. That active area could, for example, be traversed by a cathode serpentine channel or channels that travel back and forth between opposite sides of the active area, as shown in FIG. 65.

FIG. 65 depicts a cathode flow field 6516, two zones 6570, and a boundary 6572 that are similar to the zones 6470 and the boundary 6472 are shown as well. The cathode flow field 6516 has a serpentine channel 6556 that includes longer segments A extending in directions nominally perpendicular to a first set of opposing edges of the active area and shorter segments B extending in directions nominally parallel to a second set of opposing edges. The longer-length segments generally have lengths that are of the same order of magnitude as the distance between the first set of opposing edges of the active area (although potentially shortened somewhat to allow additional cathode serpentine channels to be routed in a nested or interleaved fashion). The longer segments A of the cathode serpentine channel 6556 can be seen to cross over the boundary 6572 and extend into both zones 6570. In such an arrangement, fluid that flows down a longer segment A, through a shorter segment B, and into another longer segment A that neighbors the original longer segment A, e.g., along the heavy dashed line 6574 shown in association with the leftmost two longer segments A in FIG. 65, will experience a pressure drop that is generally proportional to the sum of the lengths of the two longer segments A and the shorter segment B that joins them.

The gas flow through the cathode serpentine channel 6556, however, is not limited to staying within the cathode serpentine channel 6556. For example, as discussed earlier, the side of the cathode flow field 6516 in which the cathode serpentine channel 6556 is provided may be compressed against a porous or fibrous GDL (not shown) that provides an alternate flow path that allows gas to also or alternatively flow under partition walls 6566 that lie in between each pair of adjacent longer segments A, e.g., through the GDL that is sandwiched between the cathode flow field 6516 and an adjacent structure, e.g., an MEA. For example, the gas flow may also flow between the two longer segments A at the left of FIG. 65 via a flow path along dotted line 6576.

Generally speaking, the ratio of gas that flows along the flow path 6574 and the flow path 6576 may be biased towards gas flow along the channel flow path 6574 due to the fact that the cathode serpentine channel 6556 has a relatively large, open cross-section compared to the GDL flow path 6576. For example, the cathode serpentine channel 6556 may have a cross-section that is entirely open and that has relatively large dimensions (e.g., on the order of a millimeter or so in height and width), while the flow path offered by the GDL may only be on the order of a few hundred microns in height and be filled with the fibrous or porous material of the GDL. Put another way, the per-unit-length flow resistance of the GDL may be much higher than the per-unit-length flow resistance of the cathode serpentine channel 6556.

However, the overall flow resistance of the flow path 6574 will increase with increasing length of the longer segments A of the cathode serpentine channel 6556. Thus, the longer that the longer segments A of the cathode serpentine channel 6556 are, the higher the flow resistance along the flow path 6574, which causes the ratio of gas that flows through the flow path 6574 to the gas that flows through the flow path 6576 to decrease. In other words, shorter lengths of the longer segments A will result in less gas flow along the flow paths 6576 than longer lengths of the longer segments A.

Moreover, the flow resistance of the flow path 6574 may also increase during operation due to the potential of blockages, e.g., by liquid water or, for example, mineral deposits, within the cathode serpentine channel 6556. If such blockages occur, this will increase the flow resistance along the cathode serpentine channel, thereby causing the ratio of gas that flows through the flow path 6574 to the gas that flows through the flow path 6576 to decrease.

It will be understood that while only one flow path 6574 and one flow path 6576 are shown in FIG. 65, such flow paths may generally be replicated for similar geometrical features across the cathode flow field 6516 and such additional flow paths may have similar characteristics and behavior.

Returning to FIG. 64, it can be seen that by filling the same two zones 6470 with separate cathode serpentine channels 6456, the longer segments A of those serpentine channels 6456 may be decreased as compared with the longer segments A of the cathode serpentine channel 6556. In FIG. 64, the longer segments A of the cathode serpentine channels 6456 are approximately half the length of the longer segments A of the cathode serpentine channels 6556. Assuming that the cathode serpentine channels 6456 and 6556 are generally otherwise similar, e.g., similar cross-sectional areas, the flow resistance along the flow path 6474 will be significantly less, e.g., about 50% or so, of the flow resistance along the flow path 6574. This, in turn, increases the ratio of gas that flows through the cathode serpentine channels 6456 as opposed to leaking, for example, under peninsular walls 6466 (e.g., via flow path 6476). As the cathode serpentine channels 6456 traverse across the zones 6470 in a generally evenly distributed manner, this results in a more uniform distribution of gas across the zones 6470 than may occur in cathode flow fields such as the cathode flow field 6516.

Another aspect of the geometry shown in FIG. 64 is that the depicted cathode serpentine channels 6456 are arranged in a generally symmetric manner such that, at locations where the cathode serpentine channels in the two zones come into close proximity to each other, e.g., the shorter segments B that are adjacent to the boundary 6472, the total flow resistance along the serpentine channel from their respective inlets to those segments is generally equal, thereby resulting in a generally equal pressure drop from the inlet to each set of locations. This avoids a scenario in which two segments from different cathode serpentine channels are adjacent to one another but may have nominally different pressures that result in a pressure differential between them that may act to cause gas to cross from one such cathode serpentine channel to another.

For example, if one considers the flow resistance along the portions of the cathode serpentine channels 6456 that lie between the locations C in FIG. 64 and the fluidic inlet ports 6428, it can be seen that gas that flows through each cathode serpentine channel 6456 from the corresponding fluidic inlet port 6428 to the corresponding location C will flow along four longer segments A and three shorter segments B (and, arguably, a fourth shorter segment B that is not labeled but which leads from the fluidic inlet port 6428 to the leftmost longer segment A). Thus, the lengths of the portions of the cathode serpentine channels 6456 that are traversed by the gas flowing through the cathode serpentine channels 6456 may be generally the same and, accordingly (assuming that the cathode serpentine channels 6456 are otherwise the same, e.g., same cross-sectional dimensions), the total flow resistances between the fluidic inlet ports 6428 and the locations C may be the same. This results in the pressure drop experienced between the fluidic inlet ports 6428 and the locations C being generally the same, resulting in little or no pressure differential between the two locations C. As a result, there is little or no pressure differential present in the vicinity of the locations C that would act to cause gas from one cathode serpentine channel 6456 to flow from that cathode serpentine channel 6456 into the other cathode serpentine channel 6456. This avoids or reduces the risk or severity of a scenario where gas flowed into one zone 6470 migrates into the other zone 6470, resulting in a gas distribution across the cathode flow field 6416 that is skewed.

The symmetric arrangement of cathode serpentine channels depicted in FIG. 64 may thus, for example, be characterized as having, for each set of locations along the cathode serpentine channels where there is the least separation between them, identical or nominally identical path lengths along the serpentine paths followed by the cathode serpentine channels between their fluidic inlet ports and those locations.

A further benefit to the bilaterally symmetric arrangement of cathode serpentine channels that is evident from the above-discussed Figures is that such an arrangement allows the fluidic inlet ports and the fluidic outlet ports to be located near the centers of edges of the cathode flow fields (as opposed to at a corner). In implementations in which similar serpentine channel geometries may be used in both cathode flow fields and anode flow fields, locating the fluidic inlet ports and the fluidic outlet ports in the middle of opposing edges of the flow fields may allow the same flow field component to be used as either a cathode flow field or an anode flow field, thereby potentially reducing the number of unique parts that may be needed to assemble a particular COₓ electrolyzer cell.

FIG. 66 depicts a cathode flow field 6616 with serpentine channels arranged in a bilaterally symmetric manner. FIG. 67 depicts the same cathode flow field in a scaled-up, broken view manner to allow various features to be more easily labeled and seen. Large sections of the cathode flow field 6616 have been cut out and removed in FIG. 67, with the remaining portions moved so as to be adjacent to one another. In the implementation of FIGS. 66 and 67, the cathode flow field 6616 is divided into two zones 6670 that are separated by a boundary 6672. Each zone 6670 has a set of four cathode serpentine channels 6656 that switchback in a nested or interleaved manner between the boundary 6672 and the edge of the relevant zone 6670 that is farthest from the boundary 6672. The cathode serpentine channels 6656 each extend between a corresponding fluidic inlet port 6628 and a corresponding fluidic outlet port 6630 (it will be understood that such fluidic inlet ports 6628 and fluidic outlet ports 6630 may, in some implementations, fluidically connect with a common plenum or manifold in a stack of cells where the plenum or manifold delivers gas to all of the fluidic inlet ports simultaneously (or that receives gas from all of the fluidic outlet ports simultaneously, as appropriate).

The cathode flow field of FIGS. 66 and 67 may, for example, have an active area (generally corresponding to the area within the bounds of the depicted component in FIG. 66) on the order of 750-800 cm², e.g., 760-790 cm² or 770-780 cm², while the cathode serpentine channels 6656 themselves may, for example, each have a length of approximately 5000 to 6000 mm, e.g., 5200 to 5800 mm, 5400 to 5600 mm, 5400 to 5800 mm, or 5200 to 5600 mm. The cathode serpentine channels may each be generally rectangular or square in cross-section, e.g., having a transverse width (generally perpendicular to the direction of gas flow within the cathode serpentine channels) and/or depth that ranges from 0.5 mm to 2 mm, e.g., 0.5 mm, 0.6 mm, 0.7 mm, 0.8 mm, 0.9 mm, 1 mm, 1.1 mm, 1.2 mm, etc. In the depicted example, cathode serpentine channels 6656 are each separated from adjacent cathode serpentine channels by peninsular walls 6666 that are, for example, 0.5 mm to 2 mm in transverse width, e.g., 0.5 mm to 2 mm, e.g., 0.5 mm, 0.6 mm, 0.7 mm, 0.8 mm, 0.9 mm, 1 mm, 1.1 mm, 1.2 mm, etc. For example, the cathode serpentine channels 6656 may be approximately 0.8 mm in width and depth, separated from each other by peninsular walls of approximately 0.9 mm width, and each be approximately 5600 mm in length (thus having open channel areas of approximately 5400 mm² for each channel for zones covering an active area of 77650 mm²).

FIG. 68 depicts another cathode flow field 6816 with serpentine channels arranged in a bilaterally symmetric manner. FIG. 69 depicts the same cathode flow field 6816 in a scaled-up, broken view manner to allow various features to be more easily labeled and seen. Large sections of the cathode flow field 6816 have been cut out and removed in FIG. 69, with the remaining portions moved so as to be adjacent to one another. The implementation of FIGS. 68 and 69 is generally similar to that of FIGS. 66 and 67, with corresponding elements labeled with figure callouts sharing the last two digits in common with their counterparts in the implementation of FIGS. 66 and 67. The discussion above regarding such elements in the context of FIGS. 66 and 67 is equally applicable to those same elements in FIGS. 68 and 69 unless otherwise indicated below.

The implementation of FIGS. 68 and 69, for example, features a larger number of cathode serpentine channels 6856 in each zone 6870, e.g., seven cathode serpentine channels 6856 in each zone 6870. The cathode serpentine channels 6856 may each be on the order of 3000 mm to 3500 mm long. In the implementation shown, the cathode serpentine channels 6856 may be approximately 0.8 mm in width and depth, separated from each other by peninsular walls of approximately 0.9 mm width, and each be approximately 3200 mm in length (thus having open channel areas of approximately 2570 mm² for each channel for zones covering an active area of 77650 mm²).

### Parallel Channel Flow Fields

Another type of channel arrangement that may be used in some cathode flow fields is a parallel channel arrangement. Flow fields having a parallel channel arrangement have at least some channels that have a straight or substantially straight path between an inlet port and an outlet port. In some embodiments, all channels in a flow field having a parallel channel arrangement have a straight or substantially straight path between an inlet port and an outlet port. In some embodiments, Flow fields having a parallel channel arrangement have at least one dimension that is at least as long as the channel length of the parallel channels in the flow field. FIG. 70 depicts an example parallel channel cathode flow field. As can be seen, a cathode flow field 7016 is depicted that has a fluidic inlet port 7028 and a fluidic outlet port 7030. The fluidic inlet port 7028 and the fluidic outlet port 7030 may each be fluidically connected with corresponding plenum passages 7072, which may generally extend in directions parallel to one another. A series of parallel channels 7058 may be arranged in a linear array, with each parallel channel 7058 fluidically connected with and fluidically interposed between the two plenum passages 7072. The parallel channels 7058 may be designed to have similar flow resistances, e.g., similar or identical cross-sections and similar or identical lengths. The fluidic inlet port 7028 and the fluidic outlet port 7030 may be positioned at opposing corners of the parallel channel arrangement such that the flow paths from the fluidic inlet port 7028 to the fluidic outlet port 7030 via the parallel channels 7058 and the plenum passages 7072 are of generally equal length regardless of which parallel channel 7058 any given flow path flows through.

Cathode flow fields with parallel channel arrangements offer more direct fluid flow paths than serpentine channel arrangements for equivalent coverage areas provided. Additionally, the average distances that accumulated liquid water must be moved through in order to evacuate it from a parallel channel in such arrangements are significantly shorter in a parallel channel than in a serpentine channel for a similarly sized COₓ electrolyzer. While this is advantageous in that less energy is needed in order to evacuate liquid water from the channels, parallel channel arrangements will typically also include a larger number of potential alternate flow paths, e.g., tens or hundreds of flow paths, as compared with serpentine channel arrangements, which tend to include fewer numbers of flow paths, e.g., 2, 3, 4, or other relatively low numbers of flow paths. As discussed earlier, as the number of flow paths through a cathode flow field increases, it may be more likely that fluid flow that would normally flow through a blocked parallel channel will simply re-route itself and travel through one or more other unobstructed parallel channels within the cathode flow field rather than act to eject the liquid water that is obstructing fluid flow.

The larger numbers of parallel channels that may need to be used in parallel channel cathode flow fields may make it difficult to maintain the higher pressures and flow speeds needed within such cathode flow fields in the context of a COₓ electrolyzer without also reducing the cross-sectional area of the parallel channels in order to allow for higher pressure differentials between the two plenum passages 7072. Achieving such cross-sectional areas may prove challenging from a machining perspective and may make manufacturing of such cathode flow fields more challenging on the smaller scale. However, larger-sized cathode flow fields, e.g., ones that are sufficiently large enough to be able to support parallel, straight-channel flow fields, may allow the use of channel dimensions that are easily machinable to achieve a desired pressure drop. For example, parallel, straight-channel flow fields each having a length on the order of 1.5 meters in length and 0.2 mm² in cross-sectional area, e.g., 0.5 mm in width and 0.4 mm in depth, may allow for a pressure drop of 1.9 psi during normal operating conditions in some cathode flow fields, which may be sufficient to evacuate any accumulated water resulting from COₓ electrolyzer operation.

By way of example, some parallel channel cathode flow fields may have parallel channels that each have overall lengths of about 12 m or less or about 6 m or less. Some parallel channel cathode flow fields have parallel channels that each have an overall length of about 0.3 m or greater. In some embodiments, parallel channel cathode flow fields have channels that each have overall lengths on the order of between about 0.1 m and about 1.5 m, between about 0.1 m and about 0.8 m, between about 0.3 and about 2 m, between about 0.8 m and about 1.5 m, between about 0.1 m and about 0.45 m, between about 0.45 m and about 0.8 m, between about 0.8 m and about 1.15 m, between about 1.15 m and about 1.5 m, between about 0.1 m and about 0.275 m, between about 0.275 m and about 0.45 m, between about 0.45 m and about 0.625 m, between about 0.625 m and about 0.8 m, between about 0.8 m and about 0.975 m, between about 0.975 m and about 1.15 m, between about 1.15 m and about 1.32 m, or between about 1.32 m and about 1.5 m.

For example, such parallel channels may have widths that are between about 0.5 mm and about 2 mm, between about 0.5 mm and about 1.2 mm, between about 1.2 mm and about 2 mm, between about 0.5 mm and about 0.88 mm, between about 0.88 mm and about 1.2 mm, between about 1.2 mm and about 1.6 mm, between about 1.6 mm and about 2 mm, between about 0.5 mm and about 0.69 mm, between about 0.69 mm and about 0.88 mm, between about 0.88 mm and about 1.1 mm, between about 1.1 mm and about 1.2 mm, between about 1.2 mm and about 1.4 mm, between about 1.4 mm and about 1.6 mm, between about 1.6 mm and about 1.8 mm, or between about 1.8 mm and about 2 mm.

Such parallel channels may also have depths that are between about 0.3 mm and about 3 mm, between about 0.3 mm and about 1.6 mm, between about 1.6 mm and about 3 mm, between about 0.3 mm and about 0.98 mm, between about 0.98 mm and about 1.6 mm, between about 1.6 mm and about 2.3 mm, between about 2.3 mm and about 3 mm, between about 0.3 mm and about 0.64 mm, between about 0.64 mm and about 0.98 mm, between about 0.98 mm and about 1.3 mm, between about 1.3 mm and about 1.6 mm, between about 1.6 mm and about 2 mm, between about 2 mm and about 2.3 mm, between about 2.3 mm and about 2.7 mm, or between about 2.7 mm and about 3 mm.

Parallel channels with widths and depths such as those discussed above may result in each such parallel channel having an open surface area per channel of between about 150 mm² and about 3000 mm², between about 150 mm² and about 1600 mm², between about 1600 mm² and about 3000 mm², between about 150 mm² and about 860 mm², between about 860 mm² and about 1600 mm², between about 1600 mm² and about 2300 mm², between about 2300 mm² and about 3000 mm², between about 150 mm² and about 510 mm², between about 510 mm² and about 860 mm², between about 860 mm² and about 1200 mm², between about 1200 mm² and about 1600 mm², between about 1600 mm² and about 1900 mm², between about 1900 mm² and about 2300 mm², between about 2300 mm² and about 2600 mm², or between about 2600 mm² and about 3000 mm².

Such parallel channels may also have per-channel cross-sectional areas of between about 0.15 mm² and about 6 mm², between about 0.15 mm² and about 3.1 mm², between about 3.1 mm² and about 6 mm², between about 0.15 mm² and about 1.6 mm², between about 1.6 mm² and about 3.1 mm², between about 3.1 mm² and about 4.5 mm², between about 4.5 mm² and about 6 mm², between about 0.15 mm² and about 0.88 mm², between about 0.88 mm² and about 1.6 mm², between about 1.6 mm² and about 2.3 mm², between about 2.3 mm² and about 3.1 mm², between about 3.1 mm² and about 3.8 mm², between about 3.8 mm² and about 4.5 mm², between about 4.5 mm² and about 5.3 mm², or between about 5.3 mm² and about 6 mm²

Such parallel channels may also have total channel volumes (per channel) of between about 100 µl and about 9000 µl, between about 100 µl and about 4600 µl, between about 4600 µl and about 9000 µl, between about 100 µl and about 2300 µl, between about 2300 µl and about 4600 µl, between about 4600 µl and about 6800 µl, between about 6800 µl and about 9000 µl, between about 100 µl and about 1200 µl, between about 1200 µl and about 2300 µl, between about 2300 µl and about 3400 µl, between about 3400 µl and about 4600 µl, between about 4600 µl and about 5700 µl, between about 5700 µl and about 6800 µl, between about 6800 µl and about 7900 µl, or between about 7900 µl and about 9000 µl.

**In** some such implementations, cathode flow fields with parallel channels may also have structural characteristics relating to the thickness of the walls that are interposed between adjacent parallel channels. For example, the wall thickness in between adjacent parallel channels (and thus the distance between surfaces of those channels that are closest to one another) may be selected to be between about 0.0002 and about 0.0067, between about 0.0002 and about 0.0034, between about 0.0034 and about 0.0067, between about 0.0002 and about 0.0018, between about 0.0018 and about 0.0034, between about 0.0034 and about 0.005, between about 0.005 and about 0.0067, between about 0.0002 and about 0.001, between about 0.001 and about 0.0018, between about 0.0018 and about 0.0026, between about 0.0026 and about 0.0034, between about 0.0034 and about 0.0042, between about 0.0042 and about 0.005, between about 0.005 and about 0.0059, between about 0.0059 and about 0.0067 times the average overall length of the two adjacent parallel channels.

**In** some such parallel channel implementations having dimensional characteristics like those discussed above, the wall thickness between adjacent channels may be, for example, between about 0.15 mm and 5 mm, between about 0.15 mm and about 2.6 mm, between about 2.6 mm and about 5 mm, between about 0.15 mm and about 1.4 mm, between about 1.4 mm and about 2.6 mm, between about 2.6 mm and about 3.8 mm, between about 3.8 mm and about 5 mm, between about 0.15 mm and about 0.76 mm, between about 0.76 mm and about 1.4 mm, between about 1.4 mm and about 2 mm, between about 2 mm and about 2.6 mm, between about 2.6 mm and about 3.2 mm, between about 3.2 mm and about 3.8 mm, between about 3.8 mm and about 4.4 mm, or between about 4.4 mm and about 5 mm.

### Branching Parallel Channel Flow Fields

In some parallel channel implementations having dimensional characteristics like those discussed above, the parallel channels may be divided into separate clusters of adjacent channels that are each provided gas by a corresponding common inlet flow path (and that have similar exit flow path arrangements). Such parallel channel implementations may help ensure a more even distribution of gas within a cathode flow field. In effect, each cluster of parallel channels may represent a separate fluid flow "branch" that originates from the same starting point, such as a plenum or manifold that feeds the fluidic inlet ports that supply gas to each cluster of parallel channels).

FIG. 71 depicts a schematic of an example such parallel channel flow field. In FIG. 71, a schematic of a cathode flow field 7116 is shown. In the top half of FIG. 71, the cathode flow field 7116 is shown in a single piece, while in the bottom half, the flow paths through the cathode flow field 7116 are shown deconstructed into various sub-portions (dotted lines show the fluidic connections between these sub-portions). As can be seen, there are clusters 7178a/b/c/d of parallel channels 7158 that extend along a first direction 7186 in a parallel manner, similar to the parallel channels discussed earlier. In the depicted arrangement, the clusters 7178a/b/c/d are arranged in a bilaterally symmetric manner, e.g., with two clusters 7178a located at equidistant locations from, and on either side of, a symmetry axis 7172. The other clusters 7178b/c/d are also provided in pairs in which the clusters in each pair are each similarly equally spaced apart from the symmetry axis 7172.

The parallel channels 7158 in each cluster 7178a/b/c/d are each fluidically connected at one end with a corresponding inlet branch passage 7180 that extends in a second direction 7188 that is nominally orthogonal to the first direction 7186 and at the other end with a corresponding outlet branch passage 7182 that also extends in the second direction 7188. Each of the inlet branch passages 7180 connects with a corresponding inlet passage 7181 that leads to a corresponding fluidic inlet port 7128, while each of the outlet branch passages 7182 on the other side connects with an outlet passage 7183 that leads to a corresponding fluidic outlet port 7130. The inlet passages 7181 and outlet passages 7183 may generally extend along directions parallel to the second direction 7188 but may also include segments that extend in the first direction 7186 in order to connect with the fluidic inlet ports 7128 or the fluidic outlet ports 7130 (as appropriate), and the fluidic inlet ports 7128 and the fluidic outlet ports 7130 may each be located at locations near, and centered on (as a group), the symmetry axis 7172. While not depicted here, the fluidic inlet ports 7128 and the fluidic outlet ports 7130 may each connect with a corresponding common inlet or common outlet, as appropriate and as shown in other example flow fields herein.

When gas is flowed into the fluidic inlet ports 7128, the gas flows into the cathode flow field 7116 as separate gas flows to each of the inlet branch passages 7180 via a corresponding inlet passage 7181, at which point each gas flow may subdivide into the separate parallel channels 7158 that are in the respective cluster 7178a/b/c/d of parallel channels 7158 that fluidically connect with the inlet branch passage 7180 that those parallel channels 7158 connect with. Similarly, when the gas that flows down the parallel channels 7158 in a particular cluster 7178a/b/c/d, it exits those parallel channels 7158, where such gas flows will recombine in the outlet branch passage 7182 that connects with those parallel channels 7158 before exiting the cathode flow field 7116 via the corresponding outlet passages 7183 and fluidic outlet ports 7130.

It will be noted that the number of parallel channels 7158 that are in each cluster 7178a/b/c/d decreases the further the cluster 7178a/b/c/d is from the symmetry axis 7172. Put another way, the number of parallel channels 7158 that are in each cluster 7178a/b/c/d may generally decrease as a function of increasing flow path length from the corresponding fluidic inlet port 7128 to the corresponding inlet branch passage 7180 (although, in some instances, the number of parallel channels 7158 that are in some adjacent clusters may remain the same). Thus, a cluster 7178 of the clusters 7178a/b/c/d where gas travels along a longer inlet passage 7181 path length before reaching that cluster may have fewer parallel channels 7158 in it than a cluster 7178 of the clusters 7178a/b/c/d where gas travels along a shorter inlet passage 7181 path length before reaching it. Such a configuration allows for more even distribution of the gas that is flowed through the cathode flow field 7116. For example, due to the longer distance that gas must flow when flowing through the parallel channels 7158 that are in the clusters 7178d (due to the longer flow paths between the fluidic inlet ports 7128 and the inlet branch passages 7180 that connect with the parallel channels 7158 in the clusters 7178d), the overall flow resistance experienced by gas flowing through such parallel channels 7158 may be higher than with gas that flows through the parallel channels 7158 that are, for example, in the clusters 7178a/b/c (which flows along shorter flow path lengths and thus encounters lower flow resistance).

FIG. 72 depicts an example of a branching parallel channel flow field; FIG. 73 depicts the same branching channel flow field as in FIG. 72 but in enlarged form and with the middles of the parallel channels omitted by way of a break section.

In FIGS. 72 and 73, a cathode flow field 7216 with a parallel channel arrangement is shown. The cathode flow field 7216 includes 7 clusters 7278a/b/c/d/e/f/g of parallel channels 7258 on either side of a symmetry axis (not shown, but bisecting the cathode flow field 7216 horizontally with respect to the page orientation). The parallel channels 7258 are separated by partition walls 7266; further partition walls 7266 may define other channels of the cathode flow field 7216.

The parallel channels 7258 of each cluster 7278a/b/c/d/e/f/g are each connected at one end to corresponding inlet branch passages 7280a/b/c/d/e/f/g and at the other end to corresponding outlet branch passages 7282a/b/c/d/e/f/g, which generally extend along directions that are perpendicular to the parallel channels 7258 (only the inlet branch passages 7280 in the upper left quadrant and the outlet branch passages 7282 in the upper right quadrant of the depicted cathode flow field 7216 are called out, but it will be understood that additional inlet branch passages 7280 and outlet branch passages 7282 of similar design are visible in FIGS. 72 and 73). Each inlet branch passage 7280 may be connected via a corresponding inlet passage 7281 to one of the fluidic inlet ports 7228. Similarly, each outlet branch passage 7282 may be connected via a corresponding outlet passage 7283 to one of the fluidic outlet ports 7230..

The cathode flow field of FIGS. 72 and 73 may, for example, have an active area (generally corresponding to the area within the bounds of the depicted component in FIG. 72) on the order of 750-800 cm², e.g., 760-790 cm² or 770-780 cm², while the parallel channels 7258 themselves may, for example, each have a length of approximately 250 to 300 mm, e.g., 260 to 290 mm, 260 to 280 mm, 270 to 280 mm, 270 to 290 mm, or 270 to 280 mm. The parallel channels may each be generally rectangular or square in cross-section, e.g., having a transverse width (generally perpendicular to the direction of gas flow within the parallel channels) and/or depth that ranges from 0.5 mm to 2 mm, e.g., 0.5 mm, 0.6 mm, 0.7 mm, 0.8 mm, 0.9 mm, 1 mm, 1.1 mm, 1.2 mm, etc. In the depicted example, the parallel channels 7258 are each separated from adjacent parallel channels by partition walls 7266 that are, for example, 0.5 mm to 2 mm in transverse width, e.g., 0.5 mm to 2 mm, e.g., 0.5 mm, 0.6 mm, 0.7 mm, 0.8 mm, 0.9 mm, 1 mm, 1.1 mm, 1.2 mm, etc. For example, the parallel channels 6658 may be approximately 0.8 mm in width and 0.5 mm deep, separated from each other by partition walls of approximately 0.9 mm width, and each be approximately 270 mm in length.

FIG. 74 depicts a schematic of another example of a branching parallel channel flow field. In FIG. 74, a cathode flow field 7416 is shown in which there are multiple clusters of parallel channels 7458 (similar, for example, to the clusters 7178 depicted in FIG. 71). The parallel channels 7458 in each cluster of parallel channels 7458 may be connected at one end to an inlet branch passage 7480 and at the other end to an outlet branch passage 7482. Each inlet branch passage 7480 may be connected with a corresponding fluidic inlet port 7428 via a corresponding inlet passage 7481, and each outlet branch passage 7482 may be connected with a corresponding fluidic outlet port 7430 via a corresponding outlet passage 7483. In FIG. 74, only one inlet branch passage 7480, outlet branch passage 7482, inlet passage 7481, and outlet passage 7483 are indicated with callouts, but it will be understood that other pairs of inlet/outlet branch passages 7480/7482 and inlet/outlet passages 7481/7483 are present as well in association with each cluster of parallel channels 7458.

The arrangement of parallel channels 7458 and inlet/outlet branch passages 7480/7482 shown in FIG. 74 is very similar to that shown in FIG. 71. However, there is one significant difference-the inlet branch passages 7480 and the outlet branch passages 7482 for each cluster of parallel channels 7458 in FIG. 74 are each connected with a respective inlet passage 7481 or outlet passage 7483 at, in effect, opposite ends. For example, the inlet branch passage 7480 is connected to an inlet passage 7481 that leads to one of the fluidic inlet ports 7428, and the outlet branch passage 7482 is connected to an outlet passage 7483 that leads to one of the fluidic outlet ports 7430. However, the inlet passage 7481 leading to the fluidic inlet port 7428 connects to the inlet branch passage 7480 at a location along the inlet branch passage 7480 that is closest to that fluidic inlet port 7428, while the outlet passage 7483 leading to the fluidic outlet port 7430 connects to the outlet branch passage 7482 at a location along the outlet branch passage 7482 that is furthest from that fluidic outlet port 7430. It will be appreciated that the reverse arrangement may be used as well (essentially flipping the depicted arrangement left-to-right).

Another way of looking at this arrangement is that the inlet passage 7481 that leads from the fluidic inlet port 7428 connects with the inlet branch passage 7480 at a location that is proximate to one of the two outermost parallel channels 7458 in the cluster of parallel channels 7458 that the inlet branch passage 7480 provides gas to, while the outlet passage 7483 that leads to the fluidic outlet port 7430 connects with the outlet branch passage 7482 at a location that is proximate to the other of the two outermost parallel channels 7458 in the cluster of parallel channels 7458 that the outlet branch passage 7482 receives gas from. For clarity, the "outermost" parallel channels in a cluster of parallel channels are the two channels between which all of the other parallel channels in the cluster (if any) are located.

Such an arrangement may ensure that gas that flows into a given cluster of parallel channels 7458 will need to not only traverse along one of the parallel channels 7458 in that cluster in order to reach the fluidic outlet ports 7430, but will also need to traverse along, in aggregate, one of the inlet branch passages 7480. In effect, such an arrangement generally equalizes the flow path length from fluidic inlet port 7428 to fluidic outlet port 7430 for all of the parallel channels 7458 in a given cluster of parallel channels 7458. This serves to help equalize the flow resistance between the parallel channels 7458 within each cluster of parallel channels 7458, thereby enhancing flow uniformity within each cluster of parallel channels 7458.

FIG. 75 depicts a schematic of yet another example of a branching parallel channel flow field. In FIG. 75, a cathode flow field 7516 is shown in which there are multiple clusters of parallel channels 7558 (similar, for example, to the clusters depicted in FIG. 71). The parallel channels 7558 in each cluster of parallel channels 7558 may be connected at one end with inlet branch passages 7580 (7580' and 7580") and at the other end with outlet branch passages 7582 (7582' and 7582"). Each inlet branch passage 7580 may connect with a corresponding fluidic inlet port 7528 via a corresponding inlet passage 7581, and each outlet branch passage 7582 may connect with a corresponding outlet port 7528 via a corresponding outlet passage 7583. As shown, the outlet branch passage 7582 that is called out is actually split into two sub-portions 7582' and 7582", each of which is connected with the same outlet passage 7583 by a corresponding outlet branch passage extensions 7585 (7585' or 7585"). The lengths of these outlet branch passage extensions 7585' and 7585" may generally be equivalent. As in FIG. 74, only one inlet branch passage 7580, outlet branch passage 7582, inlet passage 7581, and outlet passage 7582 are indicated, but it will be understood that other instances of such passages may be associated with each cluster of parallel channels 7558.

The arrangement shown in FIG. 75 is similar to that shown in FIG. 74, although the inlet passages 7581 and outlet passages 7583 that connect the inlet branch passages 7580 and outlet branch passages 7582 with their respective fluidic inlet ports 7528 and fluidic outlet ports 7530 do not necessarily connect to either end of the inlet branch passages 7580 or the outlet branch passages 7582. For example, the inlet passage 7581 that connects the fluidic inlet port 7528 to the inlet branch passage 7580 connects with the inlet branch passage 7580 at a location approximately midway along its length, with some of the parallel channels 7558 in the associated cluster of parallel channels 7558 connecting with a first sub-portion 7580' of the inlet branch passage 7580 on one side of that connection point, and the other parallel channels 7558 in the associated cluster of parallel channels 7558 connecting with a second sub-portion 7580" of the inlet branch passage 7580 on the other side of that connection point. It will be noted that the outlet branch passage 7582 also follows this convention, although with the outlet branch passage 7582 sub-portions having outlet branch passage extensions 7585' and 7585" that allow the flow paths to take U-turns in between where the parallel channels 7558 connect therewith and where the outlet passage 7583 leading to the fluidic outlet port 7530 connects therewith. The outlet branch passage extensions 7585' and 7585" may, as may be seen, have lengths that are each generally equivalent to the corresponding lengths of the sub-portions 7582' and 7582"of the outlet branch passage 7582.

The inlet branch passages 7580 and the outlet branch passages 7582 of FIG. 75 may be generally characterized as having corresponding sub-portions, with the sub-portions in each pair of corresponding sub-portions being connected with opposing ends of a sub-group of parallel channels 7558 in the cluster of parallel channels 7558 associated with each of the inlet branch passages 7580 and each of the outlet branch channels 7582. Each pair of sub-portions may connect with the parallel channels 7558 that span between those sub-portions in a manner that is similar to how the parallel channels 7458 in each cluster of parallel channels connect with the corresponding inlet branch passage 7480 and outlet branch passage 7482 for that cluster of parallel channels 7458 in the implementation of FIG. 74.

For example, each inlet branch passage 7580 sub-portion and each outlet branch passage 7582 sub-portion may have a first end and a second end, with the first end of each such sub-portion being closest to the location where the corresponding inlet passage 7581 or outlet passage 7583 leading to the relevant fluidic inlet or outlet port 7528 or 7530 connects with the inlet branch passage 7580 or outlet branch passage 7582 having that sub-portion and the second end of that sub-portion being furthest along the path followed by that sub-portion from that location. The parallel channels 7558 that span between each pair of sub-portions may connect with each sub-portion at locations that are spaced-apart from one another. The sequence in which each sub-group of parallel channels 7558 connects with the two sub-portions that those parallel channels 7558 span between may be reversed between those two sub-portions. For example, the parallel channel 7558 that connects with one sub-portion at a location that is, of the various connection locations, closest to the first end of that sub-portion would connect with the other sub-portion at a location that is, of the various connection locations, furthest from the first end of the other sub-portion, and vice versa.

Such an arrangement of increased tortuosity is a refinement of the configuration discussed above with respect to FIG. 74 and allows for the gas flow across the cathode flow field 7516 to be even more evenly distributed as compared with the configuration of FIG. 74. It will be understood that while the sub-portion arrangement discussed above is only shown in FIG. 75 for the two innermost clusters of parallel channels, such a configuration may be implemented for any or all of the clusters in a branching parallel channel flow field. It will also be understood that the arrangement of FIG. 75 may be reversed from left-to-right, with the inlet branch passages having inlet branch passage extensions and the outlet branch passages having no outlet branch passage extensions.

FIG. 76 depicts an example of a cathode flow field that features branching parallel channels. FIG. 77 depicts a detail view of the left and right sides of the upper half of the cathode flow field of FIG. 76, with the remainder of the flow field omitted from view.

As can be seen in FIGS. 76 and 77, the cathode flow field 7616 features a plurality of clusters 7678a/b/c/d/e/f/g of parallel channels 7658. The cluster 7678a is actually formed of two sub-groups 7678a' and 7678a" of parallel channels 7658. The parallel channels 7658 in each cluster 7678 are each provided gas from one of the fluidic inlet ports 7628 by way of a corresponding inlet branch passage 7680a/b/c/d/e/f/g that is connected to one of the fluidic inlet ports 7628 by way of corresponding inlet passage 7681. The gas that is provided to each cluster of parallel channels 7658 then exits the corresponding cluster 7678a/b/c/d/e/f/g by way of the corresponding outlet branch passage 7680a/b/c/d/e/f/g that is connected to one of the fluidic outlet ports 7630 by way of a corresponding outlet passage 7683. The inlet branch passages 7680a outlet branch passages 7680a each have two sub-portions 7680a' and 7680a", each of which is associated with a different one of the sub-groups of parallel channels 7658 in the sub-groups 7678a' and 7678a", respectively, and the outlet branch passages 7682a similarly each have two sub-portions 7682a' and 7682a" (connected to outlet passage 7683 by corresponding outlet branch passage extensions 7685, e.g., 7685a' and 7685a"), each of which is associated with a different one of the sub-groups of parallel channels 7658 in the sub-groups 7678a' and 7678a", respectively. This arrangement is generally similar to that shown in FIG. 75 and exhibits similar uniformity behavior. Dimensional values of the various depicted features that are within the ranges indicated for the cathode flow field 7216 may, for example, provide gas flow with high uniformity and sufficient water ejection capability for use in COₓ electrolyzers.

### Interdigitated Channel Flow Fields

Another type of channel arrangement that may be used in some cathode flow fields is an interdigitated channel arrangement. FIG. 78 depicts an example interdigitated channel cathode flow field. As can be seen, a cathode flow field 7816 is depicted that has a fluidic inlet port 7828 and a fluidic outlet port 7830. The fluidic inlet port 7828 and the fluidic outlet port 7830 may each be fluidically connected with a corresponding plenum passage 7872 or 7872', respectively. The plenum passages 7872 and 7872' may generally extend along directions that are parallel to one another and may have a plurality of channels 7858 or 7858' extending away from the corresponding plenum passage 7872 or 7872' and towards the other of plenum passage 7872' or 7872, respectively (for more easy reference, the plenum passage 7872 and the channels 7858 are shaded differently than the plenum passage 7872' and the channels 7858'). Each pair of adjacent channels 7858 may have a channel 7858' interposed therebetween, and each pair of adjacent channels 7858' may have a channel 7858 interposed therebetween (thus providing two sets of interdigitated channels). In such an arrangement, each channel 7858 may be a dead-end channel that does not fluidically connect with the channels 7858' within the cathode flow field 7816. Similarly, each channel 7858' may also be a dead-end channel that does not fluidically connect with the channels 7858 within the cathode flow field 7816. However, COₓ gas is still able to pass between the two sets of channels 7858 and 7858' during use by passing underneath the walls 7848 by migrating through the cathode GDL (not shown) that is compressed between the cathode flow field 7816 and the MEA of the COₓ electrolyzer in which the cathode flow field 7816 is to be used. This under-wall flow of COₓ gas is indicated in FIG. 78 through the use of short arrows 7880 that lead from the channels 7858 to the channels 7858'. Gas flow from the fluidic inlet port 7828 and through the channels 7858, as well as gas flow from the channels 7858' to the fluidic outlet port 7830 is indicated using long arrows 7890.

Cathode flow fields with interdigitated channel arrangements may, similarly to parallel channel arrangements, offer more direct fluid flow paths than serpentine channel arrangements may provide for coverage areas that are similar to coverage area 7852, and the average distances that accumulated liquid water must be moved through in order to evacuate it from a channel in such arrangements are significantly shorter in an interdigitated channel than in a serpentine channel for a similarly sized COₓ electrolyzer. While this is advantageous in that less energy is needed in order to evacuate liquid water from the channels, parallel channel arrangements will typically also include a larger number of potential alternate flow paths, e.g., tens or hundreds of flow paths, as compared with serpentine channel arrangements, which tend to include fewer numbers of flow paths, e.g., 2, 3, 4, or other relatively low numbers of flow paths. As discussed earlier, as the number of flow paths through a cathode flow field increases, it is increasingly likely that fluid flow that would normally flow through a blocked parallel channel will simply re-route itself and travel through one or more other unobstructed parallel channels within the cathode flow field rather than act to eject the liquid water that is obstructing fluid flow. By forcing gas flow under the walls 7848, interdigitated cathode flow fields may, in essence, force COₓ gas to come into contact with portions of the cathode GDL and the MEA that are underneath the walls 7848, thereby ensuring that COₓ gas reaches such regions-in parallel and serpentine channel arrangements, COₓ gas may still come into contact with such portions of the MEA and the cathode GDL, but it is not necessarily forced to do so.

Interdigitated cathode flow fields COₓ electrolyzers may have channels with various dimensional characteristics that may make them particularly well-suited to use in the COₓ electrolyzer context, e.g., with respect to facilitating water removal from the cathode flow field.

By way of example, some interdigitated channel cathode flow fields may have interdigitated channels that have individual lengths on the order of between about 0.1 m and about 1.5 m, between about 0.1 m and about 0.8 m, between about 0.8 m and about 1.5 m, between about 0.1 m and about 0.45 m, between about 0.45 m and about 0.8 m, between about 0.8 m and about 1.15 m, between about 1.15 m and about 1.5 m, between about 0.1 m and about 0.275 m, between about 0.275 m and about 0.45 m, between about 0.45 m and about 0.625 m, between about 0.625 m and about 0.8 m, between about 0.8 m and about 0.975 m, between about 0.975 m and about 1.15 m, between about 1.15 m and about 1.32 m, or between about 1.32 m and about 1.5 m.

For example, such interdigitated channels may have widths that are between about 0.5 mm and about 2 mm, between about 0.5 mm and about 1.2 mm, between about 1.2 mm and about 2 mm, between about 0.5 mm and about 0.88 mm, between about 0.88 mm and about 1.2 mm, between about 1.2 mm and about 1.6 mm, between about 1.6 mm and about 2 mm, between about 0.5 mm and about 0.69 mm, between about 0.69 mm and about 0.88 mm, between about 0.88 mm and about 1.1 mm, between about 1.1 mm and about 1.2 mm, between about 1.2 mm and about 1.4 mm, between about 1.4 mm and about 1.6 mm, between about 1.6 mm and about 1.8 mm, or between about 1.8 mm and about 2 mm.

Such interdigitated channels may also have depths that are between about 0.3 mm and about 3 mm, between about 0.3 mm and about 1.6 mm, between about 1.6 mm and about 3 mm, between about 0.3 mm and about 0.98 mm, between about 0.98 mm and about 1.6 mm, between about 1.6 mm and about 2.3 mm, between about 2.3 mm and about 3 mm, between about 0.3 mm and about 0.64 mm, between about 0.64 mm and about 0.98 mm, between about 0.98 mm and about 1.3 mm, between about 1.3 mm and about 1.6 mm, between about 1.6 mm and about 2 mm, between about 2 mm and about 2.3 mm, between about 2.3 mm and about 2.7 mm, or between about 2.7 mm and about 3 mm.

Interdigitated channels with widths and depths such as those discussed above may result in each such interdigitated channel having an open surface area per channel of between about 150 mm² and about 3000 mm², between about 150 mm² and about 1600 mm², between about 1600 mm² and about 3000 mm², between about 150 mm² and about 860 mm², between about 860 mm² and about 1600 mm², between about 1600 mm² and about 2300 mm², between about 2300 mm² and about 3000 mm², between about 150 mm² and about 510 mm², between about 510 mm² and about 860 mm², between about 860 mm² and about 1200 mm², between about 1200 mm² and about 1600 mm², between about 1600 mm² and about 1900 mm², between about 1900 mm² and about 2300 mm², between about 2300 mm² and about 2600 mm², or between about 2600 mm² and about 3000 mm².

Such interdigitated channels may also have per-channel cross-sectional areas of between about 0.15 mm² and about 6 mm², between about 0.15 mm² and about 3.1 mm², between about 3.1 mm² and about 6 mm², between about 0.15 mm² and about 1.6 mm², between about 1.6 mm² and about 3.1 mm², between about 3.1 mm² and about 4.5 mm², between about 4.5 mm² and about 6 mm², between about 0.15 mm² and about 0.88 mm², between about 0.88 mm² and about 1.6 mm², between about 1.6 mm² and about 2.3 mm², between about 2.3 mm² and about 3.1 mm², between about 3.1 mm² and about 3.8 mm², between about 3.8 mm² and about 4.5 mm², between about 4.5 mm² and about 5.3 mm², or between about 5.3 mm² and about 6 mm²

Such interdigitated channels may also have total channel volumes (per channel) of between about 100 µl and about 9000 µl, between about 100 µl and about 4600 µl, between about 4600 µl and about 9000 µl, between about 100 µl and about 2300 µl, between about 2300 µl and about 4600 µl, between about 4600 µl and about 6800 µl, between about 6800 µl and about 9000 µl, between about 100 µl and about 1200 µl, between about 1200 µl and about 2300 µl, between about 2300 µl and about 3400 µl, between about 3400 µl and about 4600 µl, between about 4600 µl and about 5700 µl, between about 5700 µl and about 6800 µl, between about 6800 µl and about 7900 µl, or between about 7900 µl and about 9000 µl.

In some such implementations, cathode flow fields with interdigitated channels may also have structural characteristics relating to the thickness of the walls that are interposed between adjacent interdigitated channels. For example, the wall thickness in between adjacent interdigitated channels (and thus the distance between surfaces of those channels that are closest to one another) may be selected to be between about 0.0002 and about 0.0067, between about 0.0002 and about 0.0034, between about 0.0034 and about 0.0067, between about 0.0002 and about 0.0018, between about 0.0018 and about 0.0034, between about 0.0034 and about 0.005, between about 0.005 and about 0.0067, between about 0.0002 and about 0.001, between about 0.001 and about 0.0018, between about 0.0018 and about 0.0026, between about 0.0026 and about 0.0034, between about 0.0034 and about 0.0042, between about 0.0042 and about 0.005, between about 0.005 and about 0.0059, between about 0.0059 and about 0.0067 times the average overall length of the two adjacent interdigitated channels.

In some such interdigitated channel implementations having dimensional characteristics like those discussed above, the wall thickness between adjacent channels may be, for example, between about 0.15 mm and 5 mm, between about 0.15 mm and about 2.6 mm, between about 2.6 mm and about 5 mm, between about 0.15 mm and about 1.4 mm, between about 1.4 mm and about 2.6 mm, between about 2.6 mm and about 3.8 mm, between about 3.8 mm and about 5 mm, between about 0.15 mm and about 0.76 mm, between about 0.76 mm and about 1.4 mm, between about 1.4 mm and about 2 mm, between about 2 mm and about 2.6 mm, between about 2.6 mm and about 3.2 mm, between about 3.2 mm and about 3.8 mm, between about 3.8 mm and about 4.4 mm, or between about 4.4 mm and about 5 mm.

In addition to the above characteristics, some implementations of the flow field channels discussed herein for use in cathode flow fields of COₓ electrolyzers may also have certain relative dimensional constraints. For example, the ratio of the channel width to wall width of the walls in between each pair of adjacent channels or channel portions may be between about 0.08 and about 10, between about 0.08 and about 5, between about 5 and about 10, between about 0.08 and about 2.6, between about 2.6 and about 5, between about 5 and about 7.5, between about 7.5 and about 10, between about 0.08 and about 1.3, between about 1.3 and about 2.6, between about 2.6 and about 3.8, between about 3.8 and about 5, between about 5 and about 6.3, between about 6.3 and about 7.5, between about 7.5 and about 8.8, or between about 8.8 and about 10.

Similarly, the total open surface area for all channels in a flow field, or the channel if a single channel is used in the flow field, for some implementations may be between about 25% and about 80%, between about 25% and about 52%, between about 52% and about 80%, between about 25% and about 39%, between about 39% and about 52%, between about 52% and about 66%, between about 66% and about 80%, between about 25% and about 32%, between about 32% and about 39%, between about 39% and about 46%, between about 46% and about 52%, between about 52% and about 59%, between about 59% and about 66%, between about 66% and about 73%, or between about 73% and about 80%.

It will be noted that while the examples discussed herein and shown in the Figures have focused on generally square cell geometries, e.g., channels that extend across a square region defining, for instance, a cathode flow field, other implementations may feature non-square cell geometries, e.g., circular geometries, oval geometries, triangular geometries, rectangular geometries, pentagonal geometries, hexagonal geometries, etc.

It will also be noted that while the channels discussed thus far have generally had constant cross-sectional profiles (except perhaps at sharp corners, in which the profiles may grow and shrink when entering and exiting the corners, respectively), some implementations may feature channels that have variable widths and/or depths at various locations along their length. For example, in some implementations, a channel width and/or depth may be increased in a reduced flow speed region extending from the fluidic inlet port to a point in between the fluidic inlet port and the fluidic outlet port as compared with the channel width and/or depth in an increased flow speed region fluidically interposed in between the reduced flow speed region and the fluidic outlet port. The increased channel depth and/or width in the reduced flow speed region may act to expand the cross-sectional area of the channel(s) in the reduced flow speed region, thereby causing the gas flow velocity in the reduced flow speed region to decrease compared to what it is in the increased flow speed region. Similarly, the reduced channel depth and/or width in the increased flow speed region may act to reduce the cross-sectional area of the channel(s) in the increased flow speed region, thereby causing the gas flow velocity in the increased flow speed region to increase compared to what it is in the decreased flow speed region. The increased residence time of the gas in the decreased flow speed region that results from such lower flow speed may provide additional time for water that is present in the cathode GDL to evaporate and/or diffuse into the gas flowing through the channel(s) in the decreased flow speed region, thereby humidifying the gas before it flows downstream into the increased flow speed region. Such implementations may assist with reducing the likelihood that portions of the cathode GDL may dry out, thereby potentially compromising the performance of the GDL.

### Pressure Considerations

More generally, cathode flow fields for COₓ electrolyzers may benefit, e.g., in terms of providing a sufficiently high enough pressure drop that the liquid water that accumulates in the cathode flow fields at an increased rate in COₓ reduction as compared with, for example, fuel cell operation, is able to be reliably ejected from the cathode flow fields by the pressure drop, from being designed to have physical structures that result in certain physical characteristics of the cathode field. For example, the cathode channels for a COₓ electrolyzer cathode flow field may have channel dimensions, e.g., length, width, and depth, that, under the typical operating conditions of the COₓ electrolyzer, result in a pressure drop between the fluidic inlet port(s) and fluidic outlet port(s) of the cathode flow field that is between about 0.001 psi and about 4 psi, between about 0.001 psi and about 2 psi, between about 2 psi and about 4 psi, between about 0.001 psi and about 1 psi, between about 1 psi and about 2 psi, between about 2 psi and about 3 psi, between about 3 psi and about 4 psi, between about 0.001 psi and about 0.5 psi, between about 0.5 psi and about 1 psi, between about 1 psi and about 1.5 psi, between about 1.5 psi and about 2 psi, between about 2 psi and about 2.5 psi, between about 2.5 psi and about 3 psi, between about 3 psi and about 3.5 psi, between about 3.5 psi and about 4 psi, between about 0.001 psi and about 0.25 psi, between about 0.25 psi and about 0.5 psi, between about 0.5 psi and about 0.75 psi, between about 0.75 psi and about 1 psi, between about 1 psi and about 1.3 psi, between about 1.3 psi and about 1.5 psi, between about 1.5 psi and about 1.8 psi, between about 1.8 psi and about 2 psi, between about 2 psi and about 2.3 psi, between about 2.3 psi and about 2.5 psi, between about 2.5 psi and about 2.8 psi, between about 2.8 psi and about 3 psi, between about 3 psi and about 3.3 psi, between about 3.3 psi and about 3.5 psi, between about 3.5 psi and about 3.8 psi, between about 3.8 psi and about 4 psi, between about 0.001 psi and about 0.13 psi, between about 0.13 psi and about 0.25 psi, between about 0.25 psi and about 0.38 psi, between about 0.38 psi and about 0.5 psi, between about 0.5 psi and about 0.63 psi, between about 0.63 psi and about 0.75 psi, between about 0.75 psi and about 0.88 psi, between about 0.88 psi and about 1 psi, between about 1 psi and about 1.1 psi, between about 1.1 psi and about 1.3 psi, between about 1.3 psi and about 1.4 psi, between about 1.4 psi and about 1.5 psi, between about 1.5 psi and about 1.6 psi, between about 1.6 psi and about 1.8 psi, between about 1.8 psi and about 1.9 psi, between about 1.9 psi and about 2 psi, between about 2 psi and about 2.1 psi, between about 2.1 psi and about 2.3 psi, between about 2.3 psi and about 2.4 psi, between about 2.4 psi and about 2.5 psi, between about 2.5 psi and about 2.6 psi, between about 2.6 psi and about 2.8 psi, between about 2.8 psi and about 2.9 psi, between about 2.9 psi and about 3 psi, between about 3 psi and about 3.1 psi, between about 3.1 psi and about 3.3 psi, between about 3.3 psi and about 3.4 psi, between about 3.4 psi and about 3.5 psi, between about 3.5 psi and about 3.6 psi, between about 3.6 psi and about 3.8 psi, between about 3.8 psi and about 3.9 psi, or between about 3.9 psi and about 4 psi. In some other implementations, such channels for COₓ electrolyzers may have dimensions and operational conditions, e.g., fluidic inlet port pressures, that are selected so as to produce, during normal operational flow conditions for a COₓ electrolyzer, a pressure drop of between about 4 psi and about 50 psi, between about 4 psi and about 27 psi, between about 27 psi and about 50 psi, between about 4 psi and about 16 psi, between about 16 psi and about 27 psi, between about 27 psi and about 38 psi, between about 38 psi and about 50 psi, between about 4 psi and about 9.8 psi, between about 9.8 psi and about 16 psi, between about 16 psi and about 21 psi, between about 21 psi and about 27 psi, between about 27 psi and about 33 psi, between about 33 psi and about 38 psi, between about 38 psi and about 44 psi, between about 44 psi and about 50 psi, between about 4 psi and about 6.9 psi, between about 6.9 psi and about 9.8 psi, between about 9.8 psi and about 13 psi, between about 13 psi and about 16 psi, between about 16 psi and about 18 psi, between about 18 psi and about 21 psi, between about 21 psi and about 24 psi, between about 24 psi and about 27 psi, between about 27 psi and about 30 psi, between about 30 psi and about 33 psi, between about 33 psi and about 36 psi, between about 36 psi and about 38 psi, between about 38 psi and about 41 psi, between about 41 psi and about 44 psi, between about 44 psi and about 47 psi, or between about 47 psi and about 50 psi. It will be understood that the pressure drop may exceed the above ranges under certain circumstances, e.g., if the exit stream from the fluidic outlet port(s) goes to an inlet port of another electrolyzer cell, if water accumulates within a channel and obstructs flow through the channel, if the cathode GDL bulges up into the flow field channels when compressed, etc. Pressure drops lower than 0.5 psi may also work but may also increase the risk of the COₓ gas flows through the cathode flow field simply re-routing in instances where liquid water blocks a particular cathode channel (assuming multiple cathode channels are present) rather than acting to eject the liquid water from the blocked channel. Pressure drops higher than one or more of the ranges listed above may also work, but may not provide any additional performance benefit, i.e., may simply result in excess energy consumption by the COₓ electrolyzer while providing gas distribution uniformity and water ejection capability that may be provided by lower pressure drops as well. Such pressure drops are, it is to be understood, to be evaluated in the context of typical operating conditions of a COₓ electrolyzer, e.g., with a COₓ gas pressure in the range of 50 psig to 400 psig or 75 psig to 400 psig range and a gas flow velocity of 0.019 m/s to 30 m/s within at least some portions of the channels. For example, cathode flow fields such as those discussed above, or ones similar thereto, may be used in a COₓ electrolyzer cell in which COₓ-containing gas is flowed into the fluidic inlet ports of the cathode flow fields at a flow rate of between 2 sccm and 21 sccm per square centimeter of active cathode flow field area, inlet pressures of between 50 psig and 400 psig, and temperatures of between 30 °C and 80 °C. Under such conditions, such cathode flow fields may develop a pressure drop between the fluidic inlet ports and the fluidic outlet ports thereof that is sufficient to reliably eject any liquid water that may accumulate within the cathode channels, while still providing sufficiently uniform gas flow across the cathode flow field, e.g., such as the pressure drops discussed herein.

### GDL Design

COₓ electrolyzers may also benefit from use of cathode GDLs having particular characteristics and features that may assist with the transport of species between the MEA and flow field, including COₓ, dissolved bicarbonate/carbonate salts, water, and gaseous and dissolved generated byproducts. As noted earlier, a cathode GDL suitable for use in a COₓ electrolyzer may include, for example, a fibrous substrate that provides structural support, e.g., to the catalyst layer in the MEA 1105 (see, e.g., FIG. 11A). In some implementations, the cathode GDL may include a fibrous substrate, e.g., backing paper, cloth, or felt, that is made of an electrically conductive material, e.g., carbon fiber, which provides structural support to a microporous layer (MPL). The fibrous substrate may, for example, be woven (cloth) or non-woven (paper or felt). The MPL may be a porous carbon layer that ensures intimate contact between the cathode GDL and the adjacent MEA (the MPL may be on a side of the cathode GDL that faces and contacts the MEA). Example MPL materials may include polymer-integrated or polymer-supported granular carbon layers, e.g., fluoropolymer-integrated or fluoropolymer-supported carbon particle layers.

FIG. 79 depicts a partial cross-section view of an example cathode GDL and portions of an MEA and cathode flow field. The MEA 7902 is shown without any internal or structural details, and the portion of the cathode flow field 7916 that is shown includes a representative channel cross-section. Sandwiched in between the cathode flow field 7916 and the MEA 7902 is the cathode GDL 7914, which includes a fibrous layer 7976 and a microporous layer 7978. The photographs at left are magnified views of representative examples of the fibrous layer 7976 and the microporous layer 7978.

During COₓ electrolyzer operation, liquid water that is transported through the MEA from the anode side of the electrolyzer cell to the cathode side of the cell, as well as liquid water that is generated in the cathode side during COₓ reduction, may pass through the cathode GDL and into the cathode flow field channels. The cathode GDL may be selected to have particular properties in order to facilitate and encourage such liquid water ejection from the cathode GDL while maintaining a plurality of open (not liquid-filled) passages for gas diffusion and convection through the GDL. For example, the cathode GDL may have polytetrafluoroethylene (PTFE) or other hydrophobic component(s) added to both the MPL and the fibrous substrate to make the MPL and the fibrous substrate more hydrophobic, which may promote liquid water ejection from the cathode GDL and prevent water in the flow field from diffusing or otherwise transporting back to the cathode layer.

The discussion below relates to GDLs used for the cathode GDL in a COₓ electrolyzer, and, in some cases other electrolysis systems. In various of the embodiments described below the GDL includes one or more carbon components such as fibrous carbon, carbon powders at submicron scale, acetylene black, fullerene, Ketjen Black, polyacrylonitrile, and/or porous carbon. In certain embodiments, the carbon in a GDL has a density of about 75-1300 m²/g.

As discussed above, GDLs may include a fibrous layer, also referred to as a backing layer, and a microporous layer (MPL). In some embodiments, the microporous layer may overlap with or extend into the backing layer to at least some extent. In some embodiments, the microporous layer and the backing layer are affixed to one another such that they resist delamination during handling, fabrication of an electrode, and/or electrolysis. In some COₓ electrolyzers, the cathode GDL is arranged such that the MPL is in contact with or proximate to the MEA while the other side of the GDL is in contact with the cathode flow field.

There are commercial GDLs available that omit an MPL, but testing showed that in some COₓ electrolyzers, such GDLs yielded poor performance. For example, in a test that was conducted using two similar GDLs, with one GDL having an MPL and the other not, the Faradaic yield of carbon monoxide (FY_CO) in the COₓ electrolyzer dropped from about 90-100% to less than 75% in four hours and to less than 25% at around 9 hours when using the GDL without the MPL, whereas the COₓ electrolyzer using the GDL with the MPL continuously produced at least about 90% FY_CO for 16 hours. At the same time, the electrolyzer cell voltage remained steady in the COₓ cell when using the GDL with the MPL over 16 hours, while the voltage climbed steadily in the COₓ electrolyzer when using the GDL without the MPL over the same duration of time. This difference is generally understood to be associated with improved access of CO2 gas to the catalyst layer in the GDL having the MPL.

The GDL in a COₓ electrolyzer, in combination with the cathode flow field, plays a significant role in the removal of water from the COₓ electrolyzer cathode. GDLs that are selected or constructed so as to have particular characteristics may enhance the water ejection rates and/or capabilities of a COₓ electrolyzer. As noted earlier, the ability of the MEA in a COₓ electrolyzer to sustain the electrochemical reaction of CO2 to COₓ is hampered by the presence of liquid water, which is present in significant amounts during normal operation. If not adequately removed from the cathode, water degrades COₓ electrolyzer performance by influencing the mass transport of gaseous species and facilitating the production of side products such as H₂ through the electrolysis of water.

GDLs are often designed for use in fuel cells, flow batteries, and/or water electrolyzers. While such GDLs are not optimized for use in COₓ electrolyzers they can nonetheless sometimes be used in such contexts. The present inventors identified certain characteristics of GDLs that may be selected so as to provide a GDL that offers particularly effective performance in the COₓ electrolyzer context. The performance of different GDLs in the COₓ electrolyzer context often differs significantly from the performance of those same GDLs in other contexts, e.g., in fuel cells, flow batteries, and/or water electrolyzers. What works well in those other contexts may not work well in the COₓ context, and vice-versa.

For example, in the fuel cell context, it is preferable to avoid the use of thick GDLs. Fuel cells, due to the conditions under which they operate, experience reduced diffusion of reactants through the GDL to the catalyst surface with increasing thickness of the GDL. As such, many GDLs that are commercially available are in the about 300 µm, e.g., 315 µm, or less thickness range, with some suppliers possibly offering GDLs up to about 400 µm, e.g., 410 µm. Higher-thickness GDLs are generally perceived to negatively impact the performance of fuel cells and manufacturers thus generally avoid making GDLs that are thicker than 300 µm, or at most 400 µm. It will be understood that references below to specific thicknesses or thickness ranges of cathode GDLs, unless indicated otherwise, refer to the uncompressed thicknesses of such GDLs. For commercially available GDLs, the uncompressed thicknesses thereof are the typical thickness parameters used to specify such GDLs.

In contrast, COₓ electrolyzers employing thicker GDLs may not suffer from such performance degradation. COₓ electrolyzers tend to operate at higher pressures and lower temperatures than fuel cells and, as such, may increase the production and/or retention of liquid water generation within the COₓ electrolyzer cathode. However, somewhat unexpectedly, it was found that higher-thickness GDLs actually offer enhanced performance in the context of COₓ electrolyzers.

For example, the present inventors tested and modeled the performance of several different types of GDLs in the context of COₓ electrolyzers and found that increasing the thickness of the GDL, e.g., to thicknesses greater than those typically used in fuel cell GDLs, directly impacted the performance of COₓ electrolyzers in a significant and beneficial way.

For example, when the thickness of a GDL was tripled from 252 µm to 756 µm (the GDL thickness in the model was representative of the compressed thickness of the GDLs, i.e., the thickness of the GDLs when preloaded/clamped within an electrolyzer stack) in the model and all other inputs were held constant (there were at least 11 parameters that could be changed or adjusted within the model), it was found that the model predicted a 12% increase in water vapor flux through the GDL and out the flow field. Water vapor can easily be evacuated from the COₓ electrolyzer as part of the gaseous exhaust stream. While not wishing to be bound by theory, the increased water vapor flux was tied to the temperature gradient that the model indicated across the GDL. For example, the temperature at the interface between the cathode flow field and the GDL was 44 °C for both GDLs, but the temperature at the GDL/catalyst interface was 46.5 °C for the thinner GDL and 51.5 °C for the thicker GDL. The increased temperature differential may increase the water vapor flux.

Testing also showed that thicker GDLs, e.g., 350 µm or thicker (uncompressed and inclusive of MPL and backing layer) yielded more repeatable and higher performance than thinner, e.g., 200 µm (inclusive of MPL and backing layer) GDLs. For example, the Faradaic yield in a test COₓ electrolyzer remained at about 95% or greater for three 45-hour performance runs for the thicker (350 µm or greater) GDL combinations while the thinner GDL (200 µm) saw an immediate reduction in performance from the beginning of the test, e.g., dropping below 90% within about 6 hours and below 85% within about 13 hours (and never recovering above 85% for the remainder of the test). All GDLs from this set of data had 25% by weight PTFE content in the backing layer and MPL. The thicker GDLs used in the tests included GDLs having uncompressed thicknesses in the 350 to 550 µm range, 950 to 1250 µm range, and 1350 to 1750 µm range (such GDLs were composed of multiple discrete GDLs that were arranged in a stacked configuration in order to obtain the desired thicknesses, as commercially available GDLs in such thicknesses were not available-presumably due to their detrimental performance in the context of fuel cells).

Testing also showed that thicker GDLs, e.g., 600 µm or thicker (uncompressed and inclusive of MPL and backing layer) yielded more repeatable and higher performance than thinner, e.g., 315 µm (inclusive of MPL and backing layer) GDLs. For example, the FY_CO in a test COₓ electrolyzer remained at 95% or greater for two 28-hour performance runs for the thicker (600 µm) GDL while the thinner GDL (315 µm) saw comparable performance over a 15-hour period but then saw a significant and immediately apparent decrease in FY_CO performance when a second performance run was performed-dropping to 95% within about 6 hours, 90% within 11 hours, and about 85% within 21 hours. Both GDLs had 5% by weight PTFE content in the backing layer.

In this example, the thicker GDL was assembled by stacking two thinner, commercially available GDLs-one with an MPL and one without-so as to create a thicker GDL having MPL on one side (the side facing the MEA) and an expanse of backing layer on the other side (facing the cathode flow field). The backing layer portion of the stacked GDL had 5% by weight PTFE treatment throughout. The resulting 600 µm GDL was, to the inventors' knowledge and due to its thickness, a new type of GDL that was not previously available. The inventors thus created their own thick GDLs. The experiment revealed that such thicker GDLs, somewhat surprisingly, not only functioned when used in COₓ electrolyzers, but also offered significant and unexpected performance benefits.

The increased thickness of the GDL, e.g., 400 µm or more uncompressed, results in a longer heat conduction path through the GDL, which may, in turn, lead to a higher temperature differential across the GDL due to heat generated in the MEA that travels through the GDL and into the cathode flow field. This increased temperature differential causes more heat to be transferred into liquid water that may be present within the GDL and causes an increased fraction of such liquid water to transition to (or remain in) the vapor phase, thereby facilitating its removal from the GDL and improving the Faradaic yield performance of the COₓ electrolyzer.

A further test was performed with the 600 µm stacked GDL and another stacked GDL similar in construction to the 600 µm GDL but 880 µm thick (both uncompressed). In this further test, both GDLs were used in COₓ electrolyzers for periods of nearly 70 consecutive hours. While both GDLs experienced performance drops of FY_CO over that timeframe, the thicker (880 µm thick) GDL dropped from about 97% to 90% FY_CO within about 20 hours compared to the about 45 hours that it took the somewhat thinner (but still comparatively thick) GDL to reach the same FY_CO. However, the 880 µm thick GDL then stabilized and consistently operated at between about 88% and about 90% FY_CO for 50 hours or more, while the 600 µm thick GDL's FY_CO performance never stabilized and, in fact, exhibited gradually accelerating degradation as time progressed. By 60 hours, the FY_CO of the 600 µm thick GDL had dropped below 88%, and by 68 hours it had dropped below 86%. Thus, the 880 µm thick GDL provided lower, although much more consistent, performance over the 70-hour test period as compared to the somewhat thinner 600 µm GDL, which offered increasingly lower FY_CO performance over time.

In accordance with various embodiments, a GDL on the cathode side of a COₓ electrolyzer has an uncompressed thickness of at least about 300 µm, or at least about 400 µm, or at least about 501 µm. In some embodiments, a GDL on the cathode side of a COₓ electrolyzer has a thickness of about 200 µm to 1000 µm, about 300 µm to 1000 µm, about 400 µm to 1000 µm, about 501 µm to 1000 µm, about 600 µm to 1000 µm, about 200 µm to 1600 µm, about 300 µm to 1600 µm, about 400 µm to 1600 µm, about 501 µm to 1600 µm, about 600 µm to 1600 µm, about 200 µm to 2000 µm, about 300 µm to 2000 µm, about 400 µm to 2000 µm, about 501 µm to 2000 µm, about 600 µm to 2000 µm, about 200 µm to 3000 µm, about 300 µm to 3000 µm, about 400 µm to 3000 µm, about 501 µm to 3000 µm, or about 600 µm to 3000 µm. In some alternative implementations, a GDL on the cathode side of a COₓ electrolyzer may have an uncompressed thickness of about 350 to about 3000 µm, about 350 µm to about 1680 µm, about 1680 µm to about 3000 µ m , about 350 µm to about 1010 µm, about 1010 µm to about 1680 µm, about 1680 µm to about 2340 µm, about 2340 µm to about 3000 µm, about 350 µm to about 681 µm, about 681 µm to about 1010 µm, about 1010 µm to about 1340 µm, about 1340 µm to about 1680 µm, about 1680 µm to about 2010 µm, about 2010 µm to about 2340 µm, about 2340 µm to about 2670 µm, or about 2670 µm to about 3000 µm. In some further alternative implementations, a GDL on the cathode side of a COₓ electrolyzer may have an uncompressed thickness of about 400 to about 3000 µm, about 400 µm to about 1700 µm, about 1700 µm to about 3000 µm, about 400 µm to about 1050 µm, about 1050 µm to about 1700 µm, about 1700 µm to about 2350 µm, about 2350 µm to about 3000 µm, about 400 µm to about 725 µm, about 725 µm to about 1050 µm, about 1050 µm to about 1380 µm, about 1380 µm to about 1700 µm, about 1700 µm to about 2020 µm, about 2020 µm to about 2350 µm, about 2350 µm to about 2680 µm, or about 2680 µm to about 3000 µm. In some further alternative implementations, a GDL on the cathode side of a COₓ electrolyzer may have a thickness of about 450 to about 3000 µm, about 450 µm to about 1720 µm, about 1720 µm to about 3000 µm, about 450 µm to about 1090 µm, about 1090 µm to about 1720 µm, about 1720 µm to about 2360 µm, about 2360 µm to about 3000 µm, about 450 µm to about 769 µm, about 769 µm to about 1090 µm, about 1090 µm to about 1410 µm, about 1410 µm to about 1720 µm, about 1720 µm to about 2040 µm, about 2040 µm to about 2360 µm, about 2360 µm to about 2680 µm, or about 2680 µm to about 3000 µm. In some implementations, GDLs having thicknesses as presented here include one or more MPLs and one or more backing layers.

### Formation and Pre-compression of GDL Stacks

Although the benefits of thicker GDLs are apparent, the use of multiple discrete GDLs arranged in a stacked configuration to produce such thicker GDLs presents challenges with consistently assembling and testing cells, whether in a single-cell structure or a multi-cell or cell stack configuration. For instance, due, at least in part, to the intentionally heterogenous nature of both the MPL layer and the fibrous substrate to ensure adequate porosity and permeability, commercially available GDLs typically exhibit thickness variations, which may range between about 0.0017 cm and about 0.04 cm with a porosity between about 70% and about 80% by volume. Such variance may be compounded when multiple discrete GDLs are stacked to form thicker GDLs. Not only do such thickness variations create obstacles in forming accurate stochastic microstructure models to computationally determine the efficacy of one GDL configuration over another, but the variations also thwart attempts to obtain consistent test results between similarly configured prototypes.

Moreover, the variability in thickness in commercially available GDLs can lead to undesirable dimensional changes when a stack of multiple discrete GDLs is compressed during cell assembly. For example, although an amount of dimensional change is to be expected when a porous or otherwise pliable medium is compressed, the variability in thickness of a GDL (or a stack of GDLs) can not only lead to eccentric axial loading, and thereby, uneven compression, but also lead to differences in localized breakage and displacement of fibers that exacerbate the issues discussed above. In addition, the eccentric axial loading and/or differences in localized breakage and displacement of fibers can lead to translational and/or rotational displacement of one or more GDLs relative to the active area of a cell during assembly. This can cause misalignments with or impingement of an adjacent flow field, adverse interaction with a gasket (e.g., reduction in fluidic seal), etc., that can degrade performance of a COₓ electrolyzer cell. In the context of multi-cell stacks, unevenly compressed GDLs may cause compounding thickness inconsistencies that may result in assembly lean or flop, as well as the potential for over-compression to reduce such adverse conditions. It is also recognized that cell assembly may be accomplished more quickly and consistently when one thicker, pre-compressed GDL is utilized versus multiple discrete, uncompressed GDLs.

In accordance with various embodiments, one or more compression operations may be performed on a stack of multiple discrete GDLs to adhere and pre-compress the GDLs before inclusion within a cell assembly. Adherence of the GDLs to one another prior to cell compression may mitigate the potential for translational and/or rotational displacement of one or more of the GDLs relative to another GDL or other GDLs in the stack. To that end, thickness variations can be reduced, and less dimensional change may occur as a cell is fully compressed as part of a stack assembly. In some implementations, compression operation(s) may be performed at ambient temperature. Testing has demonstrated that about 2 to 6 cycles of compression, with each cycle having a duration of about 3 minutes to about 7 minutes, typically yields a sufficient level of GDL adhesion, stack pre-compression, and thickness uniformity to address issues such as those noted above. In one specific example, testing demonstrated that 3 cycles of compression for a duration of about 5 minutes each yielded a sufficient level of GDL adhesion, stack pre-compression, and thickness uniformity to address the issues outlined above. In some embodiments, one or more hot press operations may be utilized to reflow (or at least soften), if present, the polyacrylonitrile, PTFE, and/or other hydrophobic (or hydrophilic) component(s) of the MPL and/or the fibrous substrate to enable more rapid pre-compression and adherence of the GDLs to one another. It is also contemplated that, if multiple compression cycles are performed, the stack of multiple discrete GDLs may be rotated between cycles to reduce the effects of non-parallelism between pressing platens and non-uniformity of heat application. In some cases, the application of a heated load to the stack of GDLs may be accomplished under similar conditions (e.g., orientation, pressure, temperature, etc.) as would exist when a cell is assembled or operated apart from the presence of other cell components. One or more example processes to form a pre-compressed stack of GDLs will be described in association with FIGS. 80, 81, and 82.

FIG. 80 depicts a flowchart of an example process to form a pre-compressed stack of GDLs. Process 8000 of FIG. 80 will be described in association with FIGS. 81 and 82, which depict partial cross-sectional views of an example apparatus (e.g., apparatus 8100) and example system (e.g., roll-to-roll (R2R) system 8200) to form a pre-compressed stack of GDLs.

At step 8001, a stack of GDLs is prepared, such as stack 8101. For example, multiple discrete GDLs may be cut (e.g., die cut, laser cut, etc.) from a commercially available GDL source (such as a roll, sheet, etc.), and layered on one another in an orientation that would otherwise exist when the GDLs are assembled as part of a cell. For example, if the GDLs in question are directional, they may be stacked such that each GDL has a directionality that is orthogonal to the directionality of the GDL(s) immediately adjacent thereto. It is also contemplated that one or more discrete GDLs may be prepared as part of a stack with at least one pre-compressed GDL stack, or multiple pre-compressed GDL stacks may be utilized to prepare a thicker GDL stack. For descriptive convenience, it will be assumed that multiple discrete GDLs are prepared into stack 8101. In some embodiments, stack 8101 may be prepared from a plurality of input GDL rolls, such as input GDL rolls 8201, of R2R system 8200. This may not only increase manufacturing output but may also increase throughput via reductions in processing time. Depending on the type of commercially available GDL utilized and a desired thickness to be obtained, stack 8101 may include 2 to 10 discrete GDLs; however, any suitable number of GDLs may be utilized, such as 11 or more GDLs. In some embodiments, edges of the discrete GDLs may be aligned (or substantially aligned) with one another to form stack 8101.

Stack 8101 may be inserted, per step 8003, into thermal envelope 8103, such as an isothermal envelope, formed of a thermally reflective material(s). In some cases, thermal envelope 8103 may include opposing foil film covers formed of at least one of aluminum, copper, gold, silver, or the like. The foil film may have a thickness between about 0.006 mm and about 0.2 mm, between about 0.006 mm and about 0.1 mm, between about 0.1 mm and about 0.2 mm, between about 0.006 mm and about 0.054 mm, between about 0.054 mm and about 0.1 mm, between about 0.1 mm and about 0.15 mm, between about 0.15 mm and about 0.2 mm, between about 0.006 mm and about 0.03 mm, between about 0.03 mm and about 0.054 mm, between about 0.054 mm and about 0.079 mm, between about 0.079 mm and about 0.1 mm, between about 0.1 mm and about 0.13 mm, between about 0.13 mm and about 0.15 mm, between about 0.15 mm and about 0.18 mm, or between about 0.18 mm and about 0.2 mm. When inserted into thermal envelope 8103, exterior surfaces 8101a and 8101b of stack 8101 may be completely covered by corresponding interior surfaces 8103a and 8103b of thermal envelope 8103. In some embodiments, stack 8101 may be prepared between thermal layers 8203 provided via input rolls 8205 and 8207 of R2R system 8200. In this manner, exterior surfaces 8101a and 8101b of stack 8101 may be completely covered by surfaces 8203a and 8203b of thermal layers 8203. Thermal envelope 8103 and thermal layers 8203 may not only redirect and/or transfer heat uniformly (or substantially uniformly) during compression but may also prevent exterior surfaces 8101a and 8101b from adhering to surfaces 8103a, 8103b, 8203a, and 8203b. Further, it is not necessary that the layers of thermal envelope 8103 be attached to one another.

According to step 8005, thermal envelope 8103 including stack 8101 (or thermal layers 8203 with stack 8101 therebetween) may be positioned in apparatus 8100 between sacrificial cushion sheets 8105 (or sacrificial cushion layers 8209), which may be between compressing surfaces of apparatus 8100. In some embodiments, the compressing surfaces may be provided by platens (e.g., platens 8107), rollers, and/or any other suitable component. For descriptive convenience, it will be assumed that the compressing surfaces are provided by platens 8107. Sacrificial cushion layers 8209 may be provided via input rolls 8211 and 8213 of R2R system 8200. Sacrificial cushion sheets 8105 or layers 8209 may be formed of any suitably pliable material, such as PTFE, chlorotrifluoroethylene (E-CTFE), MIPELON^{™}, perfluoroalkoxy (PFA), ethylene tetrafluoroethylene (ETFE), etc. A thickness of sacrificial cushion sheets 8105 or layers 8209 may be between about 0.254 mm and about 0.508 mm, between about 0.254 mm and about 0.38 mm, between about 0.38 mm and about 0.508 mm, between about 0.254 mm and about 0.32 mm, between about 0.32 mm and about 0.38 mm, between about 0.38 mm and about 0.44 mm, between about 0.44 mm and about 0.508 mm, between about 0.254 mm and about 0.29 mm, between about 0.29 mm and about 0.32 mm, or between about 0.32 mm and about 0.35 mm. In some implementations, the thickness of sacrificial cushion sheets 8105 or layers 8209 may be between about 0.35 mm and about 0.38 mm, between about 0.38 mm and about 0.41 mm, between about 0.41 mm and about 0.44 mm, between about 0.44 mm and about 0.48 mm, between about 0.48 mm and about 0.508 mm, between about 0.254 mm and about 0.27 mm, between about 0.27 mm and about 0.29 mm, between about 0.29 mm and about 0.3 mm, between about 0.3 mm and about 0.32 mm, between about 0.32 mm and about 0.33 mm, or between about 0.33 mm and about 0.35 mm. According to some embodiments, the thickness of sacrificial cushion sheets 8105 or layers 8209 may be between about 0.35 mm and about 0.37 mm, between about 0.37 mm and about 0.38 mm, between about 0.38 mm and about 0.4 mm, between about 0.4 mm and about 0.41 mm, between about 0.41 mm and about 0.43 mm, between about 0.43 mm and about 0.44 mm, between about 0.44 mm and about 0.46 mm, between about 0.46 mm and about 0.48 mm, between about 0.48 mm and about 0.49 mm, or between about 0.49 mm and about 0.508 mm. As such, sacrificial cushion sheets 8105 or layers 8209 may enable pressure applied to thermal envelope 8103 or layers 8203 (and, thereby, to stack 8101) via platens 8107 to be more uniformly (or substantially uniformly) distributed. This may mitigate issues associated with the variability in thickness of the multiple discrete GDLs of stack 8101 and/or some non-parallelism between platens 8107.

It is also noted that sacrificial cushion layers 8209 may reduce friction between platens 8107 and thermal layers 8203 in R2R system 8200. To this end, infeed portion 8215 of R2R system 8200, apparatus 8100, and/or outfeed portion 8217 of R2R system 8200 may include one or more mechanisms (e.g., brakes, motors, rollers, sensors, tensioners, etc.) to control web speed and tension in R2R system 8200, and, thereby, to control supply of source GDL, thermal layer, and sacrificial cushion layer materials to apparatus 8100.

In some embodiments, apparatus 8100 may be a hot press, such as a Carver^{™} hot press, a laminator, and/or any other suitable thermocompression device. As such, platens 8107 may be pre-heated to a setpoint between about 20 °C and about 80 °C, between about 20 °C and about 50 °C, between about 50 °C and about 80 °C, between about 20 °C and about 35 °C, between about 35 °C and about 50 °C, between about 50 °C and about 65 °C, between about 65 °C and about 80 °C, between about 20 °C and about 28 °C, between about 28 °C and about 35 °C, between about 35 °C and about 42 °C, between about 42 °C and about 50 °C, between about 50 °C and about 57 °C, between about 57 °C and about 65 °C, between about 65 °C and about 72 °C, between about 72 °C and about 80 °C, between about 20 °C and about 24 °C, between about 24 °C and about 28 °C, between about 28 °C and about 31 °C, between about 31 °C and about 35 °C, between about 35 °C and about 39 °C, between about 39 °C and about 42 °C, between about 42 °C and about 46 °C, between about 46 °C and about 50 °C, between about 50 °C and about 54 °C, between about 54 °C and about 57 °C, between about 57 °C and about 61 °C, between about 61 °C and about 65 °C, between about 65 °C and about 69 °C, between about 69 °C and about 72 °C, between about 72 °C and about 76 °C, or between about 76 °C and about 80 °C.

According to step 8007, one or more compression operations may be performed to form a pre-compressed stack of GDLs. For example, apparatus 8100 may apply compressive force to stack 8101 by, for example, causing relative motion between press frames 8109 and 8111 via press 8113, which may be a hydraulically actuated cylinder. In some embodiments, one compression cycle is performed. In some implementations, multiple compression cycles are performed, such as 2 cycles to 10 cycles, e.g., 3 cycles to 7 cycles, for instance, 6 cycles to 8 cycles, such as 4 cycles, 5 cycles, or 9 cycles. To this end, compressive force of each cycle may be applied (e.g., progressively applied) to stack 8101 in any suitable fashion, e.g., linearly, stepwise, exponentially, or according to any other suitable pressure gradient. For example, pressure may be progressively applied from 0 psi to between about 100 psi and about 400 psi, between about 100 psi and about 250 psi, between about 250 psi and about 400 psi, between about 100 psi and about 180 psi, between about 180 psi and about 250 psi, between about 250 psi and about 320 psi, between about 320 psi and about 400 psi, between about 100 psi and about 140 psi, between about 140 psi and about 180 psi, between about 180 psi and about 210 psi, between about 210 psi and about 250 psi, between about 250 psi and about 290 psi, between about 290 psi and about 320 psi, between about 320 psi and about 360 psi, between about 360 psi and about 400 psi, between about 100 psi and about 120 psi, between about 120 psi and about 140 psi, between about 140 psi and about 160 psi, between about 160 psi and about 180 psi, between about 180 psi and about 190 psi, between about 190 psi and about 210 psi, between about 210 psi and about 230 psi, between about 230 psi and about 250 psi, between about 250 psi and about 270 psi, between about 270 psi and about 290 psi, between about 290 psi and about 310 psi, between about 310 psi and about 320 psi, between about 320 psi and about 340 psi, between about 340 psi and about 360 psi, between about 360 psi and about 380 psi, or between about 380 psi and about 400 psi. In some implementations, pressure may be progressively applied from 0 psi to between about 180 psi and about 220 psi, between about 180 psi and about 200 psi, between about 200 psi and about 220 psi, between about 180 psi and about 190 psi, between about 190 psi and about 200 psi, between about 200 psi and about 210 psi, between about 210 psi and about 220 psi, between about 180 psi and about 180 psi, between about 180 psi and about 190 psi, between about 190 psi and about 200 psi, between about 200 psi and about 200 psi, between about 200 psi and about 200 psi, between about 200 psi and about 210 psi, between about 210 psi and about 220 psi, between about 220 psi and about 220 psi, between about 180 psi and about 180 psi, between about 180 psi and about 180 psi, between about 180 psi and about 190 psi, between about 190 psi and about 190 psi, between about 190 psi and about 190 psi, between about 190 psi and about 200 psi, between about 200 psi and about 200 psi, between about 200 psi and about 200 psi, between about 200 psi and about 200 psi, between about 200 psi and about 200 psi, between about 200 psi and about 210 psi, between about 210 psi and about 210 psi, between about 210 psi and about 210 psi, between about 210 psi and about 220 psi, between about 220 psi and about 220 psi, or between about 220 psi and about 220 psi. For instance, pressure may be progressively applied from 0 psi to about 200 psi.

According to various embodiments, the maximum load of each cycle may be applied to stack 8101 for a total of between about 2 minutes and about 11 minutes, between about 2 minutes and about 6.5 minutes, between about 6.5 minutes and about 11 minutes, between about 2 minutes and about 4.2 minutes, between about 4.2 minutes and about 6.5 minutes, between about 6.5 minutes and about 8.8 minutes, between about 8.8 minutes and about 11 minutes, between about 2 minutes and about 3.1 minutes, between about 3.1 minutes and about 4.2 minutes, between about 4.2 minutes and about 5.4 minutes, between about 5.4 minutes and about 6.5 minutes, between about 6.5 minutes and about 7.6 minutes, between about 7.6 minutes and about 8.8 minutes, between about 8.8 minutes and about 9.9 minutes, between about 9.9 minutes and about 11 minutes, between about 2 minutes and about 2.6 minutes, between about 2.6 minutes and about 3.1 minutes, between about 3.1 minutes and about 3.7 minutes, between about 3.7 minutes and about 4.2 minutes, between about 4.2 minutes and about 4.8 minutes, between about 4.8 minutes and about 5.4 minutes, between about 5.4 minutes and about 5.9 minutes, between about 5.9 minutes and about 6.5 minutes, between about 6.5 minutes and about 7.1 minutes, between about 7.1 minutes and about 7.6 minutes, between about 7.6 minutes and about 8.2 minutes, between about 8.2 minutes and about 8.8 minutes, between about 8.8 minutes and about 9.3 minutes, between about 9.3 minutes and about 9.9 minutes, between about 9.9 minutes and about 10 minutes, or between about 10 minutes and about 11 minutes. For instance, the maximum load may be applied to stack 8101 for a total of about 5 minutes.

After stack 8101 is compressed for a set amount of time, a pre-compressed stack of GDLs is formed. The thickness and thickness variation of the pre-compressed stack of GDLs may be reduced relative to its uncompressed state by between about 1 % and about 30 %, between about 1 % and about 16 %, between about 16 % and about 30 %, between about 1 % and about 8.2 %, between about 8.2 % and about 16 %, between about 16 % and about 23 %, between about 23 % and about 30 %, between about 1 % and about 4.6 %, between about 4.6 % and about 8.2 %, between about 8.2 % and about 12 %, between about 12 % and about 16 %, between about 16 % and about 19 %, between about 19 % and about 23 %, between about 23 % and about 26 %, between about 26 % and about 30 %, between about 1 % and about 2.8 %, between about 2.8 % and about 4.6 %, between about 4.6 % and about 6.4 %, between about 6.4 % and about 8.2 %, between about 8.2 % and about 10 %, between about 10 % and about 12 %, between about 12 % and about 14 %, between about 14 % and about 16 %, between about 16 % and about 17 %, between about 17 % and about 19 %, between about 19 % and about 21 %, between about 21 % and about 23 %, between about 23 % and about 25 %, between about 25 % and about 26 %, between about 26 % and about 28 %, or between about 28 % and about 30 %. In some embodiments, the thickness and thickness variation of the pre-compressed stack of GDLs may be reduced relative to its uncompressed state by between about 15 % and about 18 %, between about 15 % and about 16 %, between about 16 % and about 18 %, between about 15 % and about 16 %, between about 16 % and about 17 %, between about 17 % and about 18 %, between about 15 % and about 16 %, between about 16 % and about 17 %, or between about 17 % and about 18 %. In some implementations, the thickness and thickness variation of the pre-compressed stack of GDLs may be reduced relative to its uncompressed state by between about 5.25 % and about 9.5 %, between about 5.25 % and about 7.4 %, between about 7.4 % and about 9.5 %, between about 5.25 % and about 6.3 %, between about 6.3 % and about 7.4 %, between about 7.4 % and about 8.4 %, between about 8.4 % and about 9.5 %, between about 5.25 % and about 5.8 %, between about 5.8 % and about 6.3 %, between about 6.3 % and about 6.8 %, between about 6.8 % and about 7.4 %, between about 7.4 % and about 7.9 %, between about 7.9 % and about 8.4 %, between about 8.4 % and about 9 %, or between about 9 % and about 9.5 %.

In some embodiments, the pre-compressed stack of GDLs may be optionally cut or trimmed to a predetermined size, per step 8009. For instance, a die cutter, laser cutter, wheel cutter, and/or the like may be utilized to cut or trim the pre-compressed stack of GDLs to a size appropriate for inclusion in a single or multi-cell stack assembly. In R2R system 8200, cutting mechanism 8219 may be positioned downstream from apparatus 8100 to cut appropriately sized pre-compressed stacks of GDLs from the output of apparatus 8100. Cutting mechanism 8219 may completely cut the appropriately sized pre-compressed stacks of GDLs from the output of apparatus 8100 or may form perforated cuts to enable the appropriately sized pre-compressed stacks of GDLs to be later removed from the output of apparatus 8100. Further, the output of apparatus 8100 and/or excess GDL material may be collected via output roller 8221. In a similar fashion, output rollers 8223 and 8225 may collect thermal layer material from the output of apparatus 8100. Output rollers 8227 and 8229 may collect sacrificial cushion material output from apparatus 8100.

### Additional GDL Design Considerations

Another characteristic of GDLs that may be selected so as to enhance GDL performance in the COₓ electrolyzer context is the thermal conductivity of the GDL. For example, the above-mentioned model was used to compare the predicted performance of two equal-thickness GDLs that only differed in their respective thermal conductivities, which was 0.2 W/mK in one GDL and doubled to 0.4 W/mK in the other. Halving the thermal conductivity resulted in an about 1.25 fold increase in temperature differential across the GDL, but also resulted in approximately a 105% increase in water vapor flux.

In accordance with various embodiments, a GDL on the cathode side of a COₓ electrolyzer has an average thermal conductivity of at most about 0.5 W/mK or at most about 0.1 W/mK. In some embodiments, a GDL on the cathode side of a COₓ electrolyzer has an average thermal conductivity of about 0.05 to 0.5 W/mK. In some implementations, GDLs having thermal conductivities as presented here include one or more MPLs and one or more backing layers.

In what may be at least somewhat related to the above observation regarding thermal conductivity, additional testing revealed that the presence of PTFE throughout the entire thickness of the backing layer of GDLs used in COₓ electrolyzers provided a significant performance benefit. The inclusion of PTFE in the backing layer may have any of a number of beneficial effects, including, for example, altering the hydrophobicity of the backing layer. However, the inclusion of PTFE may also decrease the thermal conductivity of the backing layer since the PTFE has a significantly lower thermal conductivity than, for example, carbon fibers that may be used in the backing layer. The PTFE may, in effect, help insulate the carbon fibers, thus lowering the thermal conductivity of the GDL as a whole.

In tests of two thicker GDLs (both about 600 µm)-one of which had 5% by weight of PTFE throughout the backing layer material and one of which had about 280 µm of backing layer with no PTFE at all-and a thinner GDL (315 µm) with 5% by weight of PTFE in the backing layer, it was found that while both GDLs with 5% by weight PTFE throughout their entire backing layer thickness maintained relatively stable and high FY_CO performance over an 18 hour test interval (greater than 85% for the 315 µm GDL, but decreasing slowly over time; greater than 95% for the 600 µm GDL over the same period and decreasing at a much slower rate) as compared with the about 600 µm GDL having PTFE only within part of the backing layer thickness. The GDL that had a portion of the backing layer thickness PTFE-free saw its FY_CO level decrease to below 85% within less than 5 hours and below 60% before 7 hours had passed. The FY_CO using this GDL dropped to less than 20% by 12 hours.

Testing also suggested that increasing the weight percent/amount of PTFE that was present within the backing layer of a GDL provided a beneficial effect in COₓ electrolyzers. In tests that were done with several GDLs, it was found that using GDLs with elevated levels of PTFE in the backing layer (e.g., 25% by weight as compared with 5% by weight) but comparable thicknesses resulted in a lower decay rate in Faradaic yield.

In accordance with various embodiments, a cathode side GDL of a COₓ electrolyzer contains a hydrophobic additive. In some such cases, the GDL or a layer thereof includes a carbonaceous material and a hydrophobic additive. In some cases, the hydrophobic additive is a hydrophobic polymer such as a fluorinated or perfluorinated polymer (e.g., PTFE). In certain embodiments, a hydrophobic additive such as a perfluorinated polymer is present in both a GDL backing layer and an MPL (both contained in the GDL). In some configurations, the hydrophobic additive is present through the entire thickness of the GDL, including an MPL, a backing layer, and any other layer. In some embodiments, a hydrophobic additive such as a perfluorinated polymer is present in a GDL at concentration of at least about 5% by weight, or about 0.5% to 55% by weight.

In some instances, it may be beneficial to use layered GDLs that have different layers, each with a different morphology and/or a different composition. As an example, each of two or more layers may comprise a backing layer and a MPL. In some embodiments, two different layers have different hydrophobic additive contents, e.g., a GDL with an MPL and three different backing layers, each with a different hydrophobic additive content, e.g., MPL/layer A/layer B/layer C, with layer A having about 5%, layer B having about 10%, and layer C having about 20% (by weight) PTFE in them.

Based on the above results and various other observations, certain potentially desirable characteristics of GDLs for use in COₓ electrolyzers were identified; these characteristics, summarized below, may be individually applicable but many or all of them may also be combinable to provide performance increases in excess of what any particular characteristic alone may be able to provide.

GDLs for use in COₓ electrolyzers may, for example, provide enhanced performance when having characteristics such as any one or more of the following:

About 200 µm-2000 µm overall thickness, with thicknesses in the 400 µm to 2000 µm range, 501 µm to 2000 µm range, or 600 µm to 900 µm range being demonstrated to provide improved performance over thinner GDLs.

About 0.5%-55% by weight PTFE content in the backing layer, with PTFE content of at least about 25% by weight in the backing layer being shown to provide good performance.

An external water contact angle having a value of about 120° to 170°, and in some implementations greater than or equal to about 140°, measured within 60 seconds of application of water for the backing layer. While this characteristic may be governed by the PTFE content of the GDL backing layer, GDLs with backing layers containing a hydrophobic material other than PTFE (e.g., other fluorinated polymers) may offer performance similar to that obtained using GDLs having PTFE content as noted above if those non-PTFE GDLs have external water contact angles within the indicated range(s).

Backing layer or overall GDL porosity of about 35% to 90% or about 60% to 90%.

Backing layer fiber diameter of about 1 µm to 25 µm, e.g., about 5 µm to 15 µm.

GDL bulk density of about 0.1 g/cm³ to 0.8 g/cm³, with bulk densities of about 0.2 g/cm³ to 0.4 g/cm³, which showed increased performance over lower bulk densities.

GDL basic weight of about 50 g/cm² to 1000 g/cm², with basic weights of about 150 g/cm² to 300 g/cm² showing increased performance over lower basic weights.

GDL area-specific resistance of about 0.05 mΩ·cm² to 20 mΩ·cm² or about 0.05 mΩ·cm² to 5 mΩ·cm².

GDL in-plane resistivity of about 0.05 mΩ·m to 7 mΩ·m or about 0.05 mΩ m to 2 mΩ m.

GDL air permeability of about 1 Gurley-second to 1000 Gurley-seconds.

GDL compressibility of about 0% to 40%, e.g., 10% to 20%.

GDL thermal conductivity of about 0.05 W/mK to 0.5 W/mK or about 0.15 W/mK to 0.35 W/mK.

GDL break strength of about 1,000 N/m to 10,000 N/m, e.g. about 2,000 N/m to 4,501 N/m.

GDL stiffness of about 20 Taber stiffness units to 40 Taber stiffness units, e.g., 25-30 Taber stiffness units.

GDL tortuosity of about 1.5 to 5 (tortuosity being the ratio of actual path length taken by molecules through GDL between two points compared to straight-line distance between those two points).

Any of the above properties may apply separately to the MPL or backing layer. Or any of the above properties may apply to both the MPL and backing layer.

As noted above, COₓ electrolyzers that use GDLs without MPLs may exhibit significantly degraded performance. Therefore, in some embodiments, at least one MPL is present in a GDL for use in a COₓ electrolyzer. In some implementations, a GDL includes at least 1 MPL, such as 2, 3, 4, or 5 MPLs, but embodiments are not limited thereto.

In some implementations, MPLs for GDLs for COₓ electrolyzer usage may have between about 15% and 55%, e.g., about 25%, by weight PTFE content. MPLs for GDLs for COₓ electrolyzer usage may also have a thickness that is in the range of about 1% to 30% of the overall thickness of the GDL.

In some implementations, a GDL comprises a stack of GDL units, each stack comprising at least one MPL affixed to at least one backing layer. In some cases, a GDL comprises a stack of two GDL units, each containing at least one backing layer and one or both of the GDL units containing an MPL. In some cases, a GDL comprises a stack of three GDL units, each GDL unit containing at least one backing layer and at least one of the GDL units containing an MPL.

It will be understood that the GDLs discussed above, e.g., in the context of cathode GDLs, may be combined with the flow fields discussed above, e.g., in the context of cathode flow fields, in a COₓ electrolyzer stack assembly. For example, the use of thicker GDLs (and/or GDLs with other characteristics discussed above) may result in higher water ejection rates from the MEAs of such an electrolyzer due to the higher water vapor flux that may occur in the context of COₓ electrolyzer use. By coupling such GDLs with flow fields such as those discussed above, which may provide superior water removal capabilities, COₓ electrolyzers may be made to operate more efficiently and with greater consistency and lower potential performance degradation due to decreased residual water retention.

One combination of the above GDL specifications that yields a high performing device has an uncompressed overall thickness of about 470-570 µm, with one microporous layer that is about 20-70 µm thick, with 25% PTFE dispersed within the microporous layer as well as the carbon fiber backing layer. This GDL may have a basis weight of about 85-90 g/m², bulk density of about 0.32-0.35 g/cm³, break strength in the machine direction of about 2100-4200 N/m, stiffness in the machine direction of about 12-52 Taber, through-plane and in-plane air permeability of about 25-50 Gurley seconds, compressibility of about 11-17%, area-specific resistivity of about 11 mOhm·cm², or any combination thereof. Note that combinations of these properties can describe various types of GDL arrangements including GDLs that comprise an MPL alone, a backing layer alone, and any stack including one or more backing layers and one or more MPLs. In some cases, the GDL having such combinations of properties comprises a stack of two more structures, each having at least one MPL and at least one backing layer.

### PTL Design

COₓ electrolyzers may also benefit from use of anode PTLs having characteristics and features that may assist with the transport of species between an anode flow field (e.g., anode flow field 1111 in FIG. 11A) and an MEA (e.g., MEA 1105 in FIG. 11A), including an anolyte such as, for example, water and/or other aqueous solutions, as well as generated byproducts of one or more reduction processes. In general, an anode PTL (such as anode PTL 1109 in FIG. 11A) may exhibit basic characteristics of electrical conductivity, thermal conductivity, surface energy, mass transport, porosity, thickness, rigidity, tensile modulus/strength, corrosion resistance, elemental abundance and manufacturability (relating to cost) and the like; however, the anode PTL may exhibit some differences from a cathode GDL, such as cathode GDL 1121 in FIG. 11A.

For example, a PTL may have a thickness sufficient for mechanical support of an MEA under cathode-over-anode differential pressures and general compression when included as part of a stack (e.g., stack 500 in FIG. 5) and compressed via, for instance, stack hardware (e.g., tensioning members 527, threaded fasteners 529, first washers 531, and/or second washers 533). Accordingly, a structure of a PTL may be generally smooth and relatively flat so as to prevent (or otherwise reduce the likelihood of) puncturing of the MEA material under non-operating and operating conditions of a stack, such as stack 500 in FIG. 5. It is also noted that the environment adjacent to the anode side of an MEA may exhibit a pH of about 0 to about 7 and oxygen evolution potential of about 1.4 V to about 2.0 V. Such an environment may be rather oxidizing, and, consequently, can be relatively aggressive (or caustic) not only to typical carbon-based GDL materials, but also various transition metals, such as yttrium (Y), zirconium (Zr), molybdenum (Mo), technetium (Tc), tantalum (Ta), hafnium (Hf), ruthenium (Ru), rhodium (Rh), palladium (Pd), platinum (Pt), silver (Ag), cadmium (Cd), etc. This may lead to relatively high rates of corrosion. Thus, a PTL (such as anode PTL 1109 in FIG. 11A) may be formed of one or more relatively corrosion-resistant, electrically conductive materials, such as titanium (Ti), niobium (Nb), and/or the like. In some embodiments, the one or more relatively corrosion-resistant, electrically conductive materials may be pure (or substantially pure) materials, e.g., pure Ti, pure Nb, etc., but embodiments are not limited thereto. Further, the one or more materials of the PTL may be sintered, printed from particles, etched, drilled or otherwise fabricated into a porous structure.

According to various implementations, the porosity of the PTL (like anode PTL 1109 in FIG. 11A) may be configured to allow for sufficient wicking of water (or other anolyte) from the bulk of adjacent flow field channels (e.g., fluidic passages 8317 and 8525 in anode flow fields 1111 described in association with FIGS. 83, 84A, 84B, and 85A-85C) to an anode catalyst layer of an MEA (such as MEA 1105 in FIG. 11A). With this in mind, the one or more materials of a PTL may not be hydrophobic and may or may not have an electroplating coating, such as an electroplating coating of, for instance, platinum (Pt), iridium (Ir), ruthenium (Ru), and/or the like. It is noted, however, that an electroplating coating may provide benefits in decreasing the electrical contact resistance of a PTL, such as anode PTL 1109 in FIG. 11A.

In various embodiments, mean particle size (e.g., particle diameter) of one or more materials forming a PTL may be between about 25 µm and about 150 µm, and mean pore size (e.g., pore diameter) may, in some implementations, be between about 10 µm and about 120 µm. Porosity may, according to various embodiments, be between about 1 % and about 90 % by volume. In some cases, a contact resistance of the PTL may be between about 5 mΩ·cm⁻² and about 50 mΩ·cm⁻², and current density may, according to various implementations, be between about 0 mA·cm⁻² and about 2000 mA·cm⁻². An average thickness of the PTL may, according to some embodiments, be between about 100 µm and about 2000 µm.

### Additional Implementations

As previously discussed, overall multi-cell stack performance may be at least partially affected by the uniformity of electrical efficiency and product selectivity across the plurality of cells of a multi-cell stack. This uniformity may very often be driven by the uniformity of gas flow delivery to/across each of the plurality of cells. To this point, the provisioning of input fluids (e.g., water, gaseous COₓ, etc.) to the plurality of cells, in that it relates to flow field pressure drop, may have a large effect on overall stack flow uniformity that may become more of an issue with increasing numbers of cells in a multi-cell stack. This is at least because the flow uniformity may improve when the pressure drop across/through the plurality of cells of a multi-cell stack is about an order of magnitude more than any pressure difference between discrete locations along a plenum where collective flow is distributed into individual cells within a multi-cell stack. Moreover, as more and more cells are included as part of a multi-cell stack, managing combined axial expansion of the plurality of cells may become more of an issue to ensure proper alignment between stack components and uniform fluid flow. Accordingly, one or more additional implementations, one or more of which may be utilized in association with stack 500 (see FIG. 6), will be described below and that may account for such considerations.

FIG. 91 depicts a perspective view of an example multi-cell COₓ electrolyzer stack. FIGS. 92 and 93 depict respective side views of the example multi-cell COₓ electrolyzer stack of FIG. 91. FIGS. 94 and 95 depict respective cross-sectional views the example multi-cell COₓ electrolyzer stack of FIG. 91 respectively taken along sectional lines 94-94 and 95-95.

Referring to FIGS. 91-95, multi-cell COₓ electrolyzer stack (or stack) 9100 includes a plurality of COₓ electrolyzer cells (or cells), such as cell 9101, formed by stacking a plurality of repeat units 9103 (individually referenced as repeat units 9103_1 to 9103_n, where "n" is an integer greater than or equal to one and "i" is an integer greater than one and less than "n") between cathode interface assembly 9105 adjacent to port side assembly 9107 and anode interface assembly 9109 adjacent to piston side assembly 9111. In one embodiment, stack 9100 may include 50 or more repeat units 9103, but it is contemplated that any suitable number of repeat units 9103 may be utilized. In a manner similar to stack 500 described in association with at least FIGS. 5-10, any given cell among the plurality of COₓ electrolyzer cells of stack 9100 may be formed by the conjunction of 1) cathode interface assembly 9105 (which includes MEA 1105 (see, e.g., cathode interface assembly 505 in FIGS. 17 and 18)) and anode components 1101 of repeat unit 9103_1 (see, e.g., anode components 1101 in FIG. 11A): 2) cathode components 1103 (which include MEA 1105 (see, e.g., cathode components 1103 in FIG. 11A)) of a first repeat unit (e.g., repeat unit 9103_1) and anode components 1101 (see, e.g., anode components 1101 in FIG. 11A) of a second repeat unit (e.g., repeat unit 9103_2) adjacent to the first repeat unit; or 3) cathode components 1103 (see, e.g., cathode components 1103 in FIG. 11A) of repeat unit 9103_n and anode interface assembly 9109. Accordingly, the MEA of any given cell among the plurality of COₓ electrolyzer cells may be configured to facilitate a COₓ reduction process, such as described in association with one or more of FIGS. 1 to 4.

It is to be appreciated that cell 9101, repeat units 9103, cathode interface assembly 9105, and anode interface assembly 9109 of stack 9100 may be configured and function equivalent (or substantially equivalent) to cell 501, repeat units 503, cathode interface assembly 505, and anode interface assembly 509 of stack 500 at least described in association with FIGS. 5-10. Further, tensioning members 9113, first and second washers 9115 and 9117, and threaded fasteners 9119 and 9121 may be configured and function equivalent (or substantially equivalent) to tensioning members 527, first and second washers 531 and 533, and threaded fasteners 529 of stack 500 at least described in association with FIGS. 5-10. As such, duplicative descriptions for cell 9101, repeat units 9103, cathode interface assembly 9105, anode interface assembly 9109, tensioning members 9113, first and second washers 9115 and 9117, and threaded fasteners 9119 and 9121 will be primarily omitted to avoid obscuring embodiments described herein. Moreover, some differences between the various components of port side assembly 9107 and piston side assembly 9111 of stack 9100 vis-à-vis port side assembly 507 and bladder side assembly 511 of stack 500 may be described below in association with FIGS. 96-109.

### Port Side Assembly

FIG. 96 depicts a perspective view of an example port side assembly of the example multi-cell COₓ electrolyzer stack of FIG. 91.

Referring to FIGS. 91-96, port side assembly 9107 may include bus plate 9601, insulation plate 9603, manifold block 9605, manifold runners 9607, and capping plate 9609 sequentially stacked from a first side of cathode interface assembly 9105 in a first direction, e.g., an axial direction, which may extend parallel to the z-axis direction shown in at least FIGS. 91-104 and 107. Hereinafter, reference to the axial direction should be understood as referring to the z-axis direction. It is noted that the first side of cathode interface assembly 9105 may face away from the plurality of repeat units 9103. Among other functions, port side assembly 9107 may at least be configured to provide one or more reactants to the cells to feed the COₓ reduction process and output one or more byproducts from the cells in association therewith.

Bus plate 9601 may be equivalent (or substantially equivalent) to bus plate 513 of stack 500 (see, e.g., FIGS. 5-10), except bus plate 9601 may include a plurality of fastener orifices 9601h, which may be countersunk with respect to surface 9601a of bus plate 9601. Insulation plate 9603 may be equivalent (or substantially equivalent) to insulation plate 517 of stack 500 (see, e.g., FIGS. 5-10), but differences will be described below in association with FIGS. 99 and 100. Manifold assembly 9611 may be similar to manifold assembly 515 of stack 500 (see, e.g., FIGS. 5-10 and 12-16), but differences will be described below in association with FIGS. 96-98.

### Port Side Assembly - Manifold Block

FIGS. 97 and 98 depict top and bottom plan views, respectively, of an example manifold block of the example port side assembly of FIG. 96.

Similar to manifold assembly 515 described in association with at least FIGS. 5-10 and 12-16, manifold assembly 9611 may be configured to provide one or more reactants to the plurality of cells of stack 9100 (see FIG. 91) to feed the COₓ reduction process(es), as well as configured to expel one or more byproducts of the COₓ reduction process(es) from the plurality of cells of stack 9100 (see FIG. 91). As such, manifold assembly 9611 may include manifold block (or main body) 9605, input and output manifold runners 9607, and one or more inlet and outlet connectors (or couplings) similar to second fluidic inlet and outlet connectors 547 and 549 of manifold assembly 515 of stack 500 (see, e.g., FIG. 5).

Referring to FIGS. 96-98, main body 9605 may be a generally rectangular plate-shaped body having first surface 9701 opposing second surface 9703 in the axial direction. Although main body 9605 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, main body 9605 will be described in association with a generally rectangular configuration. When assembled as part of stack 9100 (see FIG. 91), first surface 9701 may interface with input and output manifold runners 9607, whereas second surface 9703 may include recess 9705 configured to face and interface with insulation plate 9603. First and second surfaces 9701 and 9703 may be bounded by various peripheral surfaces (or surfaces) 9707, 9709, 9711, and 9713 that may be connected to one another via one or more other peripheral surfaces, such as peripheral surface (or surface) 9715. Embodiments, however, are not limited to the aforementioned configuration, and main body 9605 may be formed having any other suitable geometric configuration.

In some embodiments, main body 9605 may include first fluidic inlet and outlet ports 9717 and 9719 in surfaces 9701 and 9705a of recess 9705 that are configured to interface with corresponding outlet and inlet ports 96070 and 9607i of inlet and outlet manifold runners 9607, and second fluidic inlet and outlet ports 9721 and 9723 (see FIG. 95) in peripheral surfaces 9711 and 9707 that are configured to interface with fluidic inlet and outlet connectors similar to fluidic inlet and outlet connectors 547 and 549 of manifold assembly 515 (see FIG. 5). It is noted that inlet and outlet manifold runners 9607 may include inlet port 9123 as a start of one or more fluidic inlet passages 9401 (see FIG. 94) to supply, for instance, water to the anode sides of the plurality of cells of stack 9100 (see FIG. 91), and outlet port 9125 as an end of one or more fluidic outlet passages configured to expel, for instance, water from the anode sides of the plurality of cells of stack 9100 (see FIG. 91). It is noted that the one or more fluidic outlet passages may be similar to the one or more fluidic inlet passages 9401 (see FIG. 94), but may interface with outlet port 9125 versus inlet port 9123. Further, second fluidic inlet and outlet ports 9721 and 9723 may include corresponding threaded regions to engage with respective threaded regions of the inlet and outlet connectors similar to fluidic inlet and outlet connectors 547 and 549 (see, e.g., FIG. 5). Alternatively, the fluidic inlet and outlet connectors may be respectively welded, e.g., sweat welded, to second inlet and outlet ports 9721 and 9723 or otherwise coupled to second inlet and outlet ports 9721 and 9723. In this manner, second inlet port 9721 may form a starting portion of fluidic inlet passage 9501 (see FIG. 95) configured to supply, for example, gaseous COₓ to the cathode sides of the plurality of cells of stack 9100 (see FIG. 91), and second outlet port 9723 may form an ending portion of fluidic outlet passage 9503 (see FIG. 95) configured to output one or more byproducts of the COₓ reduction process of the plurality of cells of stack 9100 (see FIG. 91). Second fluidic inlet and outlet ports 9721 and 9723 (see FIG. 95) may be fluidically connected to corresponding third fluidic outlet and inlet ports 9725 and 9727 in surface 9705a via respective connecting passages 9729 and 9731 (see FIG. 95).

First surface 9701 may further include recesses 9733 and 9735 respectively encircling first fluidic inlet and outlet ports 9717 and 9719. Recesses 9733 and 9735 may be configured to receive and interface with corresponding ones of manifold runner gaskets 9613. As such, when inlet and outlet manifold runners 9607 are coupled to main body 9605 via, for example, threaded fasteners 9615, manifold runner gaskets 9613 may form corresponding fluidic seals between main body 9607 and manifold runners 9607, as well as form corresponding fluidic seals around first fluidic inlet and outlet ports 9717 and 9719. Although described as threaded fasteners, threaded fasteners 9615 may be any other suitable fastening mechanism(s), such as clips, latches, rivets, welds, etc. To this end, main body 9605 may further include fastener orifices 9737 and 9739 to engage with threaded fasteners 9615 when inlet and outlet manifold runners 9607 are coupled to main body 9605. In some cases, fastener orifices 9737 and 9739 may be threaded or otherwise configured to interface with threaded fasteners 9615.

**In** some embodiments, surface 9703 of main body 9605 may include recessed region 9705 configured to receive at least a portion of insulation plate 9603 therein when manifold assembly 9611 is incorporated as part of stack 9100 (see, e.g., FIGS. 91-95). Recessed region 9705 may terminate at surface 9705a, which may include one or more threaded openings 9743 extending into main body 9605 that are configured to threadedly engage with fasteners 9617 (e.g., flatheaded machine screws or any other suitable fastening mechanism(s)), which may be utilized to couple bus plate 9601 and insulation plate 9603 to manifold assembly 9611. Further, when manifold assembly 9611 is incorporated as part of stack 9100 and insulation plate 9603 is received in recessed region 9705 (see also FIGS. 91-95), respective fluidic seals may be formed between main body 9605 and insulation plate 9603 around first fluidic inlet and outlet ports 9717 and 9719 via gaskets 9619. Similarly, respective fluidic seals may be formed between main body 9605 and insulation plate 9603 around second fluidic outlet and inlet ports 9727 and 9725 via gaskets 9621.

Main body 9605 may further include first and second fastener orifices 9745 and 9747 arranged about a periphery of main body 9605 at one or more intervals. First and second fastener orifices 9745 and 9747 may be physically connected to one another to allow tensioning members 9113 (see, e.g., FIGS. 91-95) to pass therethrough. In this manner, main body 9605 may also function as a load-spreading member similar to end plate 519 in stack 500 (see, e.g., FIGS. 5-10). As such, main body 9605 and end plate 10107 of stack 9100 may be coupled to one another via tensioning members 9113, first and second washers 9115 and 9117, and threaded fasteners 9119 and 9121 (see, e.g., FIGS. 91-95). In some embodiments, first fastener orifices 9745 may form generally circular openings in surface 9701, and second fastener orifices 9747 may form generally oval (or generally elliptical) openings in surface 9703, but any other suitable geometric configuration may be utilized in association with first and second fastener orifices 9745 and 9747. During operation of stack 9100 (see FIG. 91), the oval shape of the openings of second fastener orifices 9747 may allow some lateral displacement of tensioning members 9113 to prevent undue stress being applied to the various components of stack 9100 as stack 9100 expands and contracts.

Main body 9605 may also include port 9749 fluidically connected to connecting passage 9731. In this manner, port 9749 may be coupled to one or more sensors to monitor a flow of fluid from the cathode sides of the plurality of cells of stack 9100 (see FIG. 95). Other features of main body 9605 (and manifold assembly 9611) may be similar to those described in association with main body 541 (and manifold assembly 515) (see FIGS. 5-10 and 12-16). It is also noted that capping plate 9609 may be coupled to manifold runners 9607 via fasteners 9623. In this manner, capping plate 9609 may include a plurality of fastener openings 9609h configured to respectively interface with fasteners 9623 and enable fasteners 9623 to engage with corresponding fastener openings in manifold runners 9607.

### Port Side Assembly - Insulation Plate

FIGS. 99 and 100 depict bottom and top plan views of an example insulation plate of the example port side assembly of FIG. 96.

Referring to FIGS. 96, 99, and 100, insulation plate 9603 may be a generally rectangular plate-shaped body having first surface 9901 (e.g., a top surface) opposing second surface 9903 (e.g., a bottom surface) in axial direction 10001, which may extend parallel (or substantially parallel) to the z-axis direction. Although insulation plate 9603 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, insulation plate 9603 will be described in association with a generally rectangular configuration. First and second surfaces 9901 and 9903 may be bounded by one or more peripheral surfaces, such as peripheral surfaces (or surfaces) 9905, 9907, 9909, and 9911 that may be connected to one another via one or more other peripheral surfaces, such as peripheral surface (or surface) 9913. In some embodiments, insulation plate 9603 may have a symmetrical configuration about one or more reference planes perpendicular to axial direction 10001. For instance, a configuration of insulation plate 9603 may be symmetrical about either or both of reference planes 10003 and 10005, but embodiments are not limited thereto.

According to various embodiments, first fluidic inlet passages 9915 and 9917 may be adjacent to peripheral edge 9909, and first fluidic outlet passages 9919 and 9921 may be adjacent to peripheral edge 9905. First fluidic inlet passages 9915 and 9917 may form portions of the one or more fluidic inlet passages 9401 (see FIG. 94) of stack 9100 in association with inlet port 9123 that provides, for instance, input water to the anode sides of the plurality of cells of stack 9100. First fluidic outlet passages 9919 and 9921 may form portions of the one or more outlet passages (that are similar to inlet passages 9401 (see FIG. 94)), but associated with output port 9125 that outputs, for instance, water from the anode sides of the plurality of cells of stack 9100. In some implementations, first fluidic inlet and outlet passages 9915-9921 may be defined by respective pluralities of orifices separated from one another via corresponding septal walls. For instance, first fluidic inlet passage 9915 may include first and second inlet orifices 9915a and 9915b separated from one another via septal wall 9901s1, whereas first fluidic outlet passage 9919 may include first and second outlet orifices 9919a and 9919b separated from one another via septal wall 9901s2. The presence of these septal walls, such as septal walls 9901s1 and 9901s2, may increase the structural rigidity and, thereby, reliability of insulation plate 9603 in the vicinity of first fluidic inlet and outlet passages 9915-9921.

According to various implementations, insulation plate 9603 may include recessed region 9923 terminating at recessed surface 9923a that is configured to receive at least a portion of bus plate 9601 (see, e.g., FIGS. 91-95) therein when bus plate 9601 and insulation plate 9603 are incorporated as part of stack 9100. Recessed region 9923 may include one or more portions (e.g., portions 9923a and 9923b) any one of which may receive terminal portion 9601t of bus plate 9601 therein. Additionally, recessed region 9923 may include one or more fastener orifices 9925 in recessed surface 9923a and extending through insulation plate 9603 that are configured to allow fasteners 9617 (e.g., flatheaded machine screws or any other suitable fastening mechanism(s)) to pass from bus plate 9601 through insulation plate 9603 and engage with fastener openings 9743 (see FIG. 98) in main body 9605 of manifold assembly 9611 to enable bus plate 9601, insulation plate 9603, and manifold assembly 9611 to be coupled to one another (see also FIGS. 91-95).

Insulation plate 9603 may also include second fluidic inlet and outlet passages 9927 and 9929, which form respective portions of inlet and outlet passages 9501 and 9503 (see FIG. 95) of stack 9100 in association with fluidic inlet and outlet ports 9721 and 9723 (see FIG. 95) of main body 9605 of manifold assembly 9611. Inlet passage 9501 (see FIG. 95) may supply one or more reactants (e.g., gaseous COₓ) to the various cathode sides of the plurality of cells of stack 9100 (see, e.g., FIGS. 91-95). Outlet passage 9503 (see FIG. 95), however, may enable one or more byproducts of the COₓ reduction process to be expelled from the various cathode sides of the plurality of cells of stack 9100 (see, e.g., FIGS. 91-95).

According to various embodiments, recesses 10007-10017 may be formed in surface 9901 of insulation plate 9603 that may be configured to respectively receive corresponding portions of gaskets 9619 and 9621 therein when, for example, insulation plate 9603 is coupled to manifold assembly 9611 via fasteners 9617 (see also FIGS. 91-95). For instance, recesses 10007 and 10009 may be formed to encircle the corresponding peripheries of first fluidic inlet passages 9915 and 9917 and interface with corresponding ones of gaskets 9619, whereas recesses 10011 and 10013 may be formed to respectively encircle the corresponding peripheries of first fluidic outlet passages 9919 and 9921 and respectively interface with corresponding ones of gaskets 9619. Further, recesses 10015 and 10017 may be formed to encircle corresponding peripheries of second fluidic inlet and outlet passages 9927 and 9929 and interface with corresponding ones of gaskets 9621.

### Piston Side Assembly

FIG. 101 depicts a perspective view of an example piston side assembly of the example multi-cell COₓ electrolyzer stack of FIG. 91 in an exploded state. FIG. 102 depicts a top plan view of the example piston side assembly of FIG. 101 in an assembled state. FIG. 103 depicts a cross-sectional view of the example piston side assembly of FIG. 102 taken along sectional line 103-103.

Referring to FIGS. 91-95 and 101-103, piston side assembly 9111 may include bus plate 10101, insulation plate 10103, piston 10105, and end plate 10107 sequentially stacked from a first side of anode interface assembly 9109 in a direction opposite the axial direction, e.g., in a direction opposite the z-axis direction. It is noted that the first side of anode interface assembly 9109 may face away from the plurality of repeat units 9103. Among other functions, piston side assembly 9111 may be at least configured to constrain axial expansion of the cells of stack 9100 during the COₓ reduction process(es) in a manner that prevents or reduces the likelihood of the plurality of cells from being overly compressed, but maintains corresponding fluidic seals and electrical conductivity between associated components of stack 9100.

Bus plate 10101 may be equivalent (or substantially equivalent) to bus plate 521 of stack 500 (see, e.g., FIGS. 5-10), except bus plate 10101 may include a plurality of fastener orifices 10101h, which may be countersunk with respect to surface 10101a of bus plate 10101. Bus plate 10101 may also include terminal portion 10101t similar to how bus plate 521 includes terminal portion 521t (see, e.g., FIGS. 5-10). Insulation plate 10103 may be equivalent (or substantially equivalent) to insulation plate 523 of stack 500 (see, e.g., FIGS. 5-10, 86, and 87), except insulation plate 10103 may exclude fastener orifices 523h, exclude fastener orifices 8633, exclude second recess 8629, include recess 10109 in surface 10103a instead of first recess 8621, and include recess 10110 (see FIG. 103) in surface 10103b. Recess 10109 may not only terminate at surface 10109a, but may also include portions 10111 and 10113 either of which may receive terminal portion 10101t of bus plate 10101 therein. Recess 10110 may be configured to receive a portion of piston 10105 therein when insulation plate 10103 and piston 10105 are incorporated as part of stack 9100. A plurality of fastener orifices 10103h corresponding to fastener orifices 10101h in bus plate 10101 may be formed in surface 10109a of recess 10109. Accordingly, when bus plate 10101 and insulation plate 10103 are assembled as part of stack 9100, at least a portion of bus plate 10101 may be received in recess 10109 of insulation plate 10103 and coupled to insulation plate 10103 via fasteners 10115 (e.g., threaded fasteners or any other suitable fastening mechanism(s)), which may extend through fastener orifices 10101h and 10103h and engage with corresponding fastener orifices 10105h formed in surface 10105a of piston 10105. As such, fastener orifices 10105h may be threaded or otherwise configured to engage with fasteners 10115. Other features, functions, materials, etc., of bus plate 10101 and insulation plate 10103 may correspond to features, functions, materials, etc., of bus plate 521 and insulation plate 517 described in association with stack 500 (see, e.g., FIGS. 5-10). End plate 10107 and piston 10105 will now be described in more detail in association with FIGS. 104-109.

### Piston Side Assembly - End Plate

FIG. 104 depicts a perspective view of an example end plate of the example piston side assembly of FIG. 101. FIGS. 105 and 106 depict a top and bottom plan views of the example end plate of FIG. 104.

Referring to FIGS. 91-95, 101, and 104-106, end plate 10107 may be a generally rectangular plate-shaped body having first surface 10401 (e.g., a top surface) opposing second surface 10403 (e.g., a bottom surface) in axial direction 10601, which extend parallel (or substantially parallel) to the z-axis direction. Although end plate 10107 is described as having a generally rectangular plate-shaped configuration, embodiments are not limited thereto and any suitable geometric configuration may be utilized, such as a generally circular, generally elliptical, generally triangular, generally pentagonal, generally hexagonal, etc., configuration. For convenience, end plate 10107 will be described in association with a generally rectangular configuration. First and second surfaces 10401 and 10403 may be bounded by one or more peripheral surfaces, such as peripheral surfaces (or surfaces) 10405, 10407, 10409, and 10411, that may be connected to one another via one or more other peripheral surfaces, such as peripheral surface (or surface) 10413. In some cases, end plate 10107 may have a symmetrical configuration about one or more reference planes perpendicular to axial direction 10601. For instance, a configuration of end plate 10107 may be symmetrical about either or both of reference planes 10603 and 10605, but embodiments are not limited thereto.

According to some implementations, end plate 10107 may include a generally rectangular protrusion 10415 extending from a first central region of first surface 10401 in axial direction 10601. Although protrusion 10415 is described as having a generally rectangular configuration, embodiments are not limited thereto and any suitable geometric configuration may be utilized, such as a generally circular, generally elliptical, generally triangular, generally pentagonal, generally hexagonal, etc., configuration. For convenience, protrusion 10415 will be described in association with a generally rectangular configuration. Protrusion 10415 may include central opening 10417 exposing surface 10419 of end plate 10107. Surface 10419 may correspond with first surface 10401, e.g., surface 10419 may form a second central region of first surface 10401 that is encircled by the first central region of first surface 10401. A plurality of protrusions 10421 may extend from surface 10419 in axial direction 10601. For instance, end plate 10107 may include nine (9) protrusions 10421 extending from surface 10419 spaced apart from one another at one or more intervals. In some embodiments, protrusions 10421 may be evenly (or substantially evenly) distributed in the area exposed by opening 10417. It is contemplated, however, that end plate 10101 may include any suitable number of protrusions, such as less than nine (9) or more than nine (9). In some implementations, protrusions 10421 may be formed as cylindrical, annular protrusions respectively including corresponding central openings 10423, but other or additional geometric configurations may be utilized. Respective upper surfaces 10425 of protrusions 10421 may be recessed from upper surface 10427 of protrusion 10415. As will become more apparent below, protrusions 10421 may be sized, shaped, located, and/or otherwise configured to enable a corresponding plurality of biasing members (e.g.. disk springs, such as Belleville springs, etc.) 10117 to be supported in opening 10417 when end plate 10107 is assembled as part of stack 9100.

End plate 10107 may also include fastener orifices 10429 through which tensioning members 9113 may pass. Tensioning members 9113 may be equivalent (or substantially equivalent) with tensioning members 527 (see, e.g., FIGS. 5-10), except tensioning members 9113 may be longer than tensioning members 527 to at least account for the presence of a greater number of repeat units 9103 than repeat units 503 in stack 500 (see, e.g., FIGS. 5-10). In some cases, fastener orifices 10429 may be arranged about a peripheral region of end plate 10107 at one or more intervals. The peripheral region may, in some implementations, be arranged between the outer surfaces of protrusion 10415 and peripheral surfaces 10405, 10407, 10409, 10411, and 10413 of end plate 10107. Some additional features of end plate 10107 will be described in association with the description of piston 10105.

### Piston Side Assembly - Piston

FIG. 107 depicts a perspective view of an example piston of the piston side assembly of FIG. 101. FIGS. 108 and 109 depict top and bottom plan views of the example piston of FIG. 107.

Referring to FIGS. 91-95, 101-103, and 107-109, piston 10105 may be a generally rectangular plate-shaped body having first surface 10701 (e.g., a top surface) opposing second surface 10703 (e.g., a bottom surface) in axial direction 10801. Although piston 10105 is described as having a generally rectangular configuration, embodiments are not limited thereto and any suitable geometric configuration may be utilized, such as a generally circular, generally elliptical, generally triangular, generally pentagonal, generally hexagonal, etc., configuration. For convenience, piston 10105 will be described in association with a generally rectangular configuration. First and second surfaces 10701 and 10703 may be bounded by one or more peripheral surfaces, such as peripheral surfaces (or surfaces) 10705, 10707, 10709, and 10711, that may be connected to one another via one or more other peripheral surfaces, such as peripheral surface (or surface) 10713. In some cases, piston 10105 may have a symmetrical configuration about one or more reference planes perpendicular to axial direction 10801, which may extend parallel (or substantially parallel) to the z-axis direction (see, e.g., FIG. 107). For instance, a configuration of piston 10105 may be symmetrical about either or both of reference planes 10803 and 10805, but embodiments are not limited thereto.

According to some implementations, piston 10105 may include a generally rectangular protrusion 10715 extending from a first central region of second surface 10703 in a direction opposite the axial direction 10801 (see FIG. 108). Although protrusion 10715 is described as having a generally rectangular configuration, embodiments are not limited thereto and any suitable geometric configuration may be utilized, such as a generally circular, generally elliptical, generally triangular, generally pentagonal, generally hexagonal, etc., configuration. For convenience, protrusion 10715 will be described in association with a generally rectangular configuration. Protrusion 10715 may terminate at surface 10717, which may be bounded by a plurality of peripheral surfaces, such as peripheral surface 10719.

A plurality of blind openings 10721 may be formed in surface 10717 and extend in axial direction 10801 towards surface 10701. The number, location, and configuration of blind openings 10721 may correspond to the number, location, and configuration of protrusions 10421 of end plate 10107 (see also FIGS. 104 and 105) such that, when piston 10105 and end plate 10107 are incorporated as part of stack 9100, respective blind openings 10721 may be concentrically aligned (or substantially concentrically aligned) with corresponding protrusions 10421 (see, e.g., FIG. 103). Respective depths of blind openings 10721 from surface 10717 in axial direction 10801 may, in some implementations, be smaller than corresponding heights of protrusions 10421 from surface 10419 in axial direction 10601 (see FIGS. 104-106), which may correspond with axial direction 10801. As such, the respective depths of blind openings 10721 may correspond to a maximum (or substantially maximum) amount of axial expansion that stack 9100 may be permitted to experience when stack 9100 is pressured. It is also noted that respective widths of blind openings 10721 in a direction perpendicular to axial direction 10801 may be greater than corresponding widths of protrusions 10421 in a direction perpendicular to axial direction 10601 (see FIGS. 104-106), but smaller than corresponding widths of biasing members 10117 in a direction perpendicular to central axis 10121 (see FIG. 101). Thus, when piston 10105 is caused to axially translate along central axis 10121 towards end plate 10107, respective protrusions 10421 may be received in corresponding blind openings 10721, and biasing members 10117 may be compressed between surface 10717 of protrusion 10715 of piston 10105 and surface 10419 of end plate 10107. In this manner, biasing members 10117 may provide a first amount of axial compression to the plurality of cells of stack 9100 when stack 9100 is not pressurized, e.g., when stack 9100 is in a cooled, non-operational state.

Piston 10105 may also include a plurality of recesses 10723 formed in the peripheral surfaces (e.g., peripheral surface 10719) of protrusion 10715. Corresponding depths of recesses 10723 may extend inwards from a respective peripheral surface of protrusion 10715 towards blind openings 10721. In some embodiments, the plurality of recesses 10723 may include first and second recesses 10723a and 10723b, but embodiments are not limited thereto. For instance, protrusion 10715 may include one recess in some cases, or include three or more recesses in other cases. The plurality of recesses 10723 may be configured to interface with a corresponding plurality of piston gaskets 10119, which may include, for instance, first and second piston gaskets 10119a and 10119b.

With reference to FIGS. 91-109, when piston 10105, end plate 10107, and piston gaskets 10119 are incorporated as part of piston side assembly 9111 of stack 9100, at least a portion of protrusion 10715 of piston 10105 may be received in opening 10417 of end plate 10107 in a manner that protrusion 10715 and opening 10417 become aligned (or substantially aligned) along central axis 10121 of piston side assembly 9111. To this end, piston gaskets 10119 may form corresponding fluidic seals between recesses 10723 of piston 10105 and inner sidewalls (such as inner sidewall 10417sw) of opening 10417 of end plate 10107. As such, a fluidically sealed cavity (or cavity) 10301 may be formed between piston 10105 and end plate 10107. In a manner similar to bladder side assembly 511 (see, e.g., FIGS. 5-10 and 90), one or more control fluids (e.g., gaseous COₓ) may be introduced to cavity 10301 to regulate a distance between surface 10717 of protrusion 10715 of piston 10105 and surface 10419 of end plate 10107.

In some embodiments, the one or more control fluids may be flowed into cavity 10301 via fluidic inlet ports 10303 and 10305 formed in peripheral surfaces 10409 and 10405 of end plate 10107. Fluidic inlet port 10303 may be fluidically connected to blind orifice 10501 formed in surface 10419 of end plate 10107 via connecting passage 10307, whereas fluidic inlet port 10305 may be fluidically connected to blind orifice 10503 formed in surface 10419 of end plate 10107 via connecting passage 10309. In this manner, the one or more control fluids may be caused to flow into cavity 10301 via the conjunction of fluidic inlet ports 10303 and 10305, connecting passages 10307 and 10309, and blind orifices 10501 and 10503, as well as source 10311 of the one or more control fluids. In some embodiments, source 10311 of the one or more control fluids may be the same as the source of input providing, for instance, gaseous COₓ, to the cathode sides of the cells of stack 9100. Regardless of the source, the distance between surface 10717 of protrusion 10715 of piston 10105 and surface 10419 of end plate 10107 may be controlled based on an accumulated pressure of the one or more control fluids in cavity 10301. In this manner, regulating the distance between surface 10717 of protrusion 10715 of piston 10105 and surface 10419 of end plate 10107 may be utilized to constrain axial expansion of the plurality of cells, such as cell 9101, during operation. This may help maintain corresponding fluidic seals and electrical conductivity between associated components of stack 9100, and, thereby, provide a second amount of axial compression to the plurality of cells of stack 9100 when stack 9100 is pressurized, e.g., in an operational state of stack 9100.

According to some embodiments, when the accumulated pressure in cavity 10301 builds beyond a determined threshold, the distance between surface 10717 of piston 10105 and surface 10419 of end plate 10107 may increase to point at which fluidic seals formed in association with piston gaskets 10119 may become compromised. If and when the fluidic seals formed in association with piston gaskets 10119 become compromised, at least some of the one or more control fluids may escape (or bleed) from cavity 10301 that may cause the accumulated pressure to decrease, and, as such, the distance between surface 10717 of piston 10105 and surface 10419 of end plate 10107 to also decrease. Such a configuration may be utilized to prevent over compression of the various components of stack 9100.

As described above, fluidic inlet ports 10303 and 10305 may be utilized to introduce one or more control fluids to cavity 10301, but a corresponding fluidic outlet port may not be provided (apart from piston gaskets 10119 becoming compromised and allowing at least some of the one or more control fluids to escape from cavity 10301). In this manner, the conjunction of piston 10105, end plate 10107, and piston gaskets 10119 may form a "dead-headed" piston in which the one or more control fluids are caused to remain in cavity 10301 until a flow of the one or more control fluids is terminated and the one or more control fluids in cavity 10301 are allowed to backflow out of one or both of fluidic inlet ports 10303 and 10305. In some cases, one or both of fluidic inlet ports 10303 and 10305 (or another fluidic port) may be additionally (or alternatively) configured as a fluidic outlet port, which may interface with, for instance, a pressure relief valve configured to release, bleed-off, or otherwise exhaust accumulated pressure in cavity 10301 in response to the accumulated pressure reaching a threshold pressure and/or based on a control signal received from a controller. Such a configuration may enable finer regulation of the accumulated pressure in cavity 10301 that may, in turn, allow for finer control over the constriction of the axial expansion of the plurality of cells of stack 9100 when stack 9100 is pressurized.

According to some embodiments, source 10311 may be configured to supply the gaseous COₓ to second fluidic inlet port 9721 (see, e.g., FIG. 95) at a first pressure and to supply the one or more control fluids (e.g., gaseous COₓ) to fluidic inlet ports 10303 and 10305 at a second pressure. In some implementations, the first and second pressures may be equivalent or substantially equivalent. In some cases, source 10311 may be configured to control (e.g., adjust) one or more of the first and second pressures based on conditions of stack 9100, e.g., based on an extent of expansion of one or more cells of stack 9100 in the axial direction, based on an accumulated pressure in cavity 10301, based on the temperature of one or more components of stack 9100, and/or the like. As such, the first and second pressures may reach equilibrium, such as, in response to steady state conditions. It is also noted that source 10311 may be configured to supply the gaseous COₓ to second fluidic inlet port 9721 (see, e.g., FIG. 95) at a first time and to supply the one or more control fluids (e.g., gaseous COₓ) to fluidic inlet ports 10303 and 10305 at a second time. In some embodiments, the first and second times may occur simultaneously or substantially simultaneously. In some cases, source 10311 may be configured to delay the supply of the one or more control fluids to fluidic inlet ports 10303 and 10305 with respect to the provisioning of the gaseous COₓ to second fluidic inlet port 9721 (see, e.g., FIG. 95). For example, source 10311 may be configured to delay the supply of the one or more control fluids to fluidic inlet ports 10303 and 10305 until one or more conditions are satisfied, e.g., an extent of expansion of one or more cells of stack 9100 in the axial direction reaches one or more defined thresholds, a temperature of one or more components of stack 9100 reaches one or more defined thresholds, flow of the gaseous COₓ to second fluidic inlet port 9721 (see, e.g., FIG. 95) reaches steady state, and/or the like.

## Claims

1. A COₓ electrolyzer apparatus (500) comprising:
a first end assembly comprising a first end plate (519) and a cathode interface assembly (505) a second end assembly comprising a second end plate (525),
an anode interface assembly (509), and a bladder gasket (559),
wherein the second end assembly is coupled to the first end assembly via a plurality of tensioning members (527);
a plurality of separator plates (1107); and
a plurality of COₓ electrolyzer cells (501) that are each formed of a plurality of repeat units (503, 1100),
wherein the plurality of cells are interposed between the first and second end assemblies and arranged in a stack along an axial direction, each cell among the cells (501) comprising an instance of first components and an instance of second components,
wherein the first components comprise:
a membrane electrode assembly (MEA; 301, 401) having a cathodic part (303, 403) an anodic part (305,405),
and a separator between the cathodic part and the anodic part;
a cathode frame (1131) adjacent to the cathodic part; and
a cathode flow field (1127) at least partially disposed in a first opening in the cathode frame,
wherein the second components comprise:
an anode frame (1115) adjacent to the anodic part of the MEA; and
an anode flow field (1111) at least partially disposed in a second opening in the anode frame,
wherein each repeat unit (503, 1100) among the repeat units comprises:
an instance of the first components;
an instance of the second components; and
the separator plate (1107) that is interposed between the cathode frame (1131) of that instance of the first components and the anode frame (1115) of that instance of the second components, the separator plate (1107) being interposed between that instance of the first components and that instance of the second components;
wherein the cathode interface assembly (505) comprises:
an instance of the first components; and
a cathode interface separator plate (1701) interposed between the first end plate and a first repeat unit among the repeat units (503, 1100);
wherein the anode interface assembly (509) comprises:
an instance of the second components; and
an anode interface separator plate (4703) interposed between a second repeat unit among the repeat units and the second end plate;
wherein the cathode (1131) and anode frames (1115) of adjacent cells among the cells are coupled to one another via a corresponding plurality of frame fasteners with a separator plate among the separator plates (1107) interposed therebetween, the frame fasteners being different from the tensioning members (527);
a first end cell is formed between the cathode interface assembly (505) and the instance of the second components of the first repeat unit, the first end cell being interposed between the first end plate and the plurality of cells (501);
a second end cell is formed between the instance of the first components of the second repeat unit and the anode interface assembly (509),
the second end cell being interposed between the plurality of cells (501) and the second end plate;
an insulation plate (523) comprising:
a first recess formed in a central portion of the insulation plate;
a second recess encircling a central region of the central portion, the second recess supporting the bladder gasket (559) therein; and
an orifice (8631) configured to receive one or more control fluids; a bus plate (521) slidably disposed in the first recess and configured to abut against the bladder gasket (559) and/or a surface of the first recess facing the bus plate (521) in the axial direction; and
a distance in the axial direction between the bus plate and the surface of the first recess facing the bus plate in the axial direction is configured to increase in response to accumulation of the one or more control fluids in an area between the bus plate and the insulation plate that is fluidically sealed via at least the bladder gasket.

2. The apparatus (500) of claim 1, wherein:
the first components further comprise a cathode gas diffusion layer (GDL) adjacent to the cathode frame (1131) and covering the cathode flow field (1127),
the cathode GDL and the cathode flow field being configured to guide a flow of gaseous COₓ across the first opening in a first direction transverse to the axial direction and in a distributed manner with respect to at least a second direction transverse to each of the axial and first directions; and
the second components further comprise an anode porous transport layer (PTL) adjacent to the anode frame (1115) and covering the anode flow field (1111), the anode PTL and the anode flow field (1111) being configured to guide a flow of anolyte across the second opening in a third direction transverse to the axial direction and in a distributed manner with respect to at least the second direction.

3. The apparatus (500) of claim 1, wherein the cathode frame (1131) comprises:
the first opening arranged in a central portion of the cathode frame;
at least one first fluidic inlet passage (2815, 2817) fluidically connected to the anodic parts of the cells;
at least one first fluidic outlet passage (2819, 2821) fluidically connected to the anodic parts of the cells;
at least one second fluidic inlet passage (2827) fluidically connected to the first opening; and
at least one second fluidic outlet passage (2829) fluidically connected to the first opening.

4. The apparatus (500) of claim 3, wherein:
the cathode frame (1131) comprises a first surface facing the MEA and a second surface facing away from the first surface; and
the second surface of the cathode frame (1131) comprises:
at least one first protrusion through which the at least one first fluidic inlet passage (2815, 2817) extends;
at least one second protrusion through which the at least one first fluidic outlet (2819, 2821) passage extends;
at least one third protrusion through which the at least one second fluidic inlet (2827) passage extends; and
at least one fourth protrusion through which the at least one second fluidic outlet (2829) passage extends.

5. The apparatus (500) of claim 4, wherein:
the at least one first protrusion of the cathode frame (1131) is arranged and configured to extend through the at least one first hole in a first separator plate among the separator plates (1107) and abut against the anode frame (1115) of a first adjacent cell among the cells (501) such that the at least one first fluidic inlet passage (2815, 2817) of the cathode frame is substantially aligned in the axial direction with the at least one third fluidic inlet passage of the anode frame of the first adjacent cell;
the at least one second protrusion of the cathode frame (1131) is arranged and configured to extend through the at least one second hole in the first separator plate and abut against the anode frame (1115) of the first adjacent cell such that the at least one first fluidic outlet passage of the cathode frame is substantially aligned in the axial direction with the at least one third fluidic outlet passage of the anode frame of the first adjacent cell;
the at least one third protrusion of the cathode frame (1131) is arranged and configured to extend through the at least one third hole in the first separator plate and abut against the anode frame (1115) of the first adjacent cell such that the at least one second fluidic inlet passage of the cathode frame is substantially aligned in the axial direction with the at least one fourth fluidic inlet passage of the anode frame of the first adjacent cell; and
the at least one fourth protrusion of the cathode frame (1131) is arranged and configured to extend through the at least one fourth hole in the first separator plate and abut against the anode frame (1115) of the first adjacent cell such that the at least one second fluidic outlet passage of the cathode frame is substantially aligned in the axial direction with the at least one fourth fluidic outlet passage of the anode frame (1115) of the first adjacent cell.

6. The apparatus (500) of claim 1, wherein:
the cathode frame (1131) further comprises a plurality of first cathode fastener orifices (2837) arranged about a peripheral area of the cathode frame, the peripheral area encircling the first opening of the cathode frame; and
the anode frame (1115) further comprises:
a plurality of first anode fastener orifices (3761) arranged about a peripheral area of the anode frame, the peripheral area encircling the second opening of the anode frame, the first cathode fastener orifices being substantially aligned with the first anode fastener orifices in the axial direction; and
a plurality of first swage nuts (1135), each first swage nut among the first swage nuts being disposed in one or the other of a corresponding one of the first anode fastener orifices and a corresponding one of the first cathode fastener orifices, the first swage nuts being configured to interface with corresponding frame fasteners among the frame fasteners.

7. The apparatus (500) of claim 2, wherein:
the first components further comprise:
a first support frame (1123) interposed between the cathode GDL and the cathode frame (1131),
the first support frame comprising a first frame opening exposing a portion of the cathode GDL to the cathode flow field, the portion of the cathode GDL abutting against the cathode flow field; and
a second support frame (1125) interposed between the MEA and the anode PTL, the second support frame comprising a second frame opening exposing a portion of the MEA to the anode PTL, the portion of the MEA abutting against the anode PTL; and
the first support frame, the cathode GDL, the MEA, and the second support frame form a unitized MEA assembly (301, 401).

8. The apparatus (500) of claim 7, wherein:
the first components further comprise:
a first cathode gasket (1129) interposed between the first support frame and the cathode frame (1131),
the first cathode gasket encircling the first opening in the cathode frame to form a first fluidic seal around the cathode flow field; and
a second cathode gasket (1133) interposed between a first separator plate among the separator plates and the cathode frame, the second cathode gasket encircling the first opening in the cathode frame (1131) to form a second fluidic seal around the cathode flow field;
the second components further comprise:
a first anode gasket set (1113); and
a second anode gasket set (1117);
the first anode gasket set (1113) comprises:
a first anode gasket interposed between the second support frame and the anode frame (1115),
the first anode gasket encircling the second opening in the anode frame to form a first fluidic seal around the anode flow field;
at least one second anode gasket interposed between the cathode frame (1131) and
the anode frame (1115),
the at least one second anode gasket encircling the at least one first fluidic inlet passage of the cathode frame and the at least one third fluidic inlet passage of the anode to form at least one fluidic seal;
at least one third anode gasket interposed between the cathode frame (1131) and the anode frame (1115),
the at least one third anode gasket encircling the at least one first fluidic outlet passage in the cathode frame and the at least one third fluidic outlet passages in the anode frame to form at least one fluidic seal;
at least one fourth anode gasket interposed between the cathode frame (1131) and
the anode frame (1115), the at least one third anode gasket encircling the at least one second fluidic inlet passage in the cathode frame and the at least one fourth fluidic inlet passage in the anode frame to form at least one fluidic seal; and
at least one fifth anode gasket interposed between the cathode frame (1131) and the anode frame (1115),
the at least one fifth anode gasket encircling the at least one second fluidic outlet passage and the at least one fourth fluidic outlet passage in the anode frame to form at least one fluidic seal; and
the second anode gasket set (1117) comprises:
a sixth anode gasket interposed between the anode frame and a second separator plate among the separator plates, the sixth anode gasket encircling the second opening in the anode frame to form a second fluidic seal around the anode flow field (1111);
at least one seventh anode gasket interposed between the anode frame and the second separator plate, the at least one seventh anode gasket encircling the at least one first hole in the second separator plate and the at least one third fluidic inlet passage in the anode frame to form at least one fluidic seal;
at least one eighth anode gasket interposed between the anode frame and the second separator plate, the at least one eighth anode gasket encircling the at least one second hole in the second separator plate and the at least one third fluidic outlet passage in the anode frame to form at least one fluidic seal;
at least one ninth anode gasket interposed between the anode frame and the second separator plate, the at least one ninth anode gasket encircling the at least one third hole in the second separator plate and the at least one fourth fluidic inlet passage in the anode frame to form at least one fluidic seal; and
at least one tenth anode gasket interposed between the anode frame and the second separator plate, the at least one ninth anode gasket encircling the at least one fourth hole in the second separator plate and the at least one fourth fluidic outlet passage in the anode frame to form at least one fluidic seal.

9. The apparatus (500) of claim 1, wherein:
each of the separator plates (1107) comprises:
a plurality of fastener orifices through which the frame fasteners respectively extend;
at least one first hole through which an inlet anolyte flow path extends;
at least one second hole through which an outlet anolyte flow path extends;
at least one third hole through which an inlet gaseous COₓ flow path extends; and
at least one fourth hole through which an outlet COₓ reduction byproduct flow path extends;
the first end assembly further comprises a first insulation plate, a manifold, and a first bus plate between the first end plate and the cathode interface assembly;
the manifold comprises:
at least one first inlet fluidically connected to the anodic parts of the cells via the inlet anolyte flow path;
at least one first outlet fluidically connected to the anodic parts of the cells via the outlet anolyte flow path;
at least one second inlet fluidically connected to the cathodic parts of the cells via the inlet gaseous COₓ flow path; and
at least one second outlet fluidically connected to the cathodic parts of the cells via the outlet COₓ reduction byproduct flow path;
the first bus plate is configured to receive a first electric potential;
the first insulation plate is configured to electrically insulate the first end plate from the first bus plate, wherein the inlet anolyte flow path, the outlet anolyte flow path, the inlet gaseous COₓ flow path, and the outlet COₓ reduction byproduct flow path do not extend into the bus plate and the first insulation plate.

10. The apparatus (500) of claim 1, wherein:
the second end assembly further comprises a second bus plate and a second insulation plate sequentially stacked in the axial direction between the anode interface assembly 509 and the second end plate;
the second bus plate is configured to receive a second electric potential; and
the second insulation plate is configured to electrically insulate the second end plate from the second bus plate.

11. The apparatus (500) of claim 10, wherein:
the second end plate comprises:
a first main body;
a second end plate protrusion extending from the first main body in the axial direction; and
a second end plate opening extending into a central portion of the second end plate protrusion in a direction opposite the axial direction and terminating at a recessed surface facing the cells;
the second end assembly further comprises a piston 10105 interposed between the second insulation plate and the second end plate, the piston comprising:
a second main body; and
a piston protrusion extending from the second main body in the direction opposite the axial direction and terminating at a protruded surface facing the recessed surface;
at least a portion of the piston protrusion is slidably disposed in at least a portion of the second end plate opening;
the second end plate further comprises one or more orifices fluidically connected to the second end plate opening, the one or more orifices being configured to receive one or more control fluids;
the piston protrusion comprises a plurality of piston gaskets 10119 encircling the piston protrusion and offset from one another in the axial direction, the piston gaskets interfacing with one or more inner sidewalls of the second end plate opening such that the second end plate opening, the piston protrusion, and the piston gaskets 10119 form a cavity within the second end assembly; and
a distance in the axial direction between the protruded surface and recessed surface is configured to increase in response to accumulation of the one or more control fluids in the cavity.

12. The apparatus (500) of claim 11, wherein:
the second end assembly further comprises a plurality of biasing members (10117);
the piston protrusion comprises a plurality of piston protrusion openings extending into the protruded surface in the axial direction;
the second end plate further comprises a plurality of support protrusions extending in the axial direction from the recessed surface and arranged in correspondence with the piston protrusion openings;
the biasing members (10117) are respectively supported in the second end plate opening via corresponding support protrusions among the support protrusions such that, in a first compressed state of the second end assembly, the biasing members are compressed between the protruded surface and the recessed surface and respective portions of the support protrusions at least partially extend into corresponding piston protrusion openings among the piston protrusion openings;
the second end plate further comprises one or more orifices fluidically connected to the second end plate opening, the one or more orifices being configured to receive one or more control fluids;
the piston protrusion comprises a plurality of piston gaskets (10119) encircling the piston protrusion and offset from one another in the axial direction, the piston gaskets interfacing with one or more inner sidewalls of the second end plate opening such that the second end plate opening, the piston protrusion, and the piston gaskets form a cavity within the second end assembly; and
a distance in the axial direction between the protruded surface and recessed surface is configured to increase in response to accumulation of the one or more control fluids in the cavity.

## Patentansprüche

1. COₓ-Elektrolyseur-Vorrichtung (500), umfassend:
eine erste Endbaugruppe, umfassend eine erste Endplatte (519) und eine Kathodengrenzflächenbaugruppe (505) eine zweite Endbaugruppe, umfassend eine zweite Endplatte (525), eine Anodengrenzflächenbaugruppe (509) und eine Blasendichtung (559), wobei die zweite Endbaugruppe über eine Vielzahl von Spannelementen (527) an die erste Endbaugruppe gekoppelt ist;
eine Vielzahl von Separatorplatten (1107); und
eine Vielzahl von COₓ-Elektrolyseur-Zellen (501), die jeweils aus einer Vielzahl von Wiederholungseinheiten (503, 1100) gebildet sind, wobei die Vielzahl von Zellen zwischen die erste und die zweite Endbaugruppe zwischengeschaltet und in einem Stapel entlang einer axialen Richtung angeordnet ist, wobei jede Zelle aus den Zellen (501) eine Instanz von ersten Komponenten und eine Instanz von zweiten Komponenten umfasst,
wobei die ersten Komponenten Folgendes umfassen:
eine Membranelektrodenbaugruppe (MEA; 301, 401), die einen kathodischen Teil (303, 403) einen anodischen Teil (305, 405) und einen Separator zwischen dem kathodischen Teil und dem anodischen Teil aufweist;
einen Kathodenrahmen (1131) benachbart zu dem kathodischen Teil; und
ein Kathodenströmungsfeld (1127), das mindestens teilweise in einer ersten Öffnung in dem Kathodenrahmen vorgesehen ist,
wobei die zweiten Komponenten Folgendes umfassen:
einen Anodenrahmen (1115) benachbart zu dem anodischen Teil der MEA; und
ein Anodenströmungsfeld (1111), das mindestens teilweise in einer zweiten Öffnung in dem Anodenrahmen vorgesehen ist,
wobei jede Wiederholungseinheit (503, 1100) aus den Wiederholungseinheiten Folgendes umfasst:
eine Instanz der ersten Komponenten;
eine Instanz der zweiten Komponenten; und
die Separatorplatte (1107), die zwischen den Kathodenrahmen (1131) dieser Instanz der ersten Komponenten und den Anodenrahmen (1115) dieser Instanz der zweiten Komponenten zwischengeschaltet ist, wobei die Separatorplatte (1107) zwischen diese Instanz der ersten Komponenten und diese Instanz der zweiten Komponenten zwischengeschaltet ist;
wobei die Kathodengrenzflächenbaugruppe (505) Folgendes umfasst:
eine Instanz der ersten Komponenten; und
eine Kathodengrenzflächenseparatorplatte (1701), die zwischen die erste Endplatte und eine erste Wiederholungseinheit aus den Wiederholungseinheiten (503, 1100) zwischengeschaltet ist;
wobei die Anodengrenzflächenbaugruppe (509) Folgendes umfasst:
eine Instanz der zweiten Komponenten; und
eine Anodengrenzflächenseparatorplatte (4703), die zwischen eine zweite Wiederholungseinheit aus den Wiederholungseinheiten und die zweite Endplatte zwischengeschaltet ist;
wobei der Kathodenrahmen (1131) und der Anodenrahmen (1115) von benachbarten Zellen aus den Zellen über eine entsprechende Vielzahl von Rahmenbefestigungsmitteln aneinandergekoppelt sind, wobei eine Separatorplatte aus den Separatorplatten (1107) dazwischen zwischengeschaltet ist, wobei sich die Rahmenbefestigungsmittel von den Spannelementen (527) unterscheiden;
eine erste Endzelle zwischen der Kathodengrenzflächenbaugruppe (505) und der Instanz der zweiten Komponenten der ersten Wiederholungseinheit gebildet ist, wobei die erste Endzelle zwischen die erste Endplatte und die Vielzahl von Zellen (501) zwischengeschaltet ist;
eine zweite Endzelle zwischen der Instanz der ersten Komponenten der zweiten Wiederholungseinheit und der Anodengrenzflächenbaugruppe (509) gebildet ist, wobei die zweite Endzelle zwischen die Vielzahl von Zellen (501) und die zweite Endplatte zwischengeschaltet ist;
eine Isolierungsplatte (523), umfassend:
eine erste Vertiefung, die in einem mittigen Abschnitt der Isolierungsplatte gebildet ist;
eine zweite Vertiefung, die eine mittige Region des mittigen Abschnitts umschließt, wobei die zweite Vertiefung die Blasendichtung (559) darin stützt; und
einen Durchlass (8631), der dazu konfiguriert ist, ein oder mehrere Steuerfluide aufzunehmen;
eine Busplatte (521), die verschiebbar in der ersten Vertiefung vorgesehen ist und dazu konfiguriert ist, an der Blasendichtung (559) und/oder einer Fläche der ersten Vertiefung, die der Busplatte (521) in der axialen Richtung zugewandt ist, anzuliegen; und
ein Abstand in der axialen Richtung zwischen der Busplatte und der Fläche der ersten Vertiefung, die der Busplatte in der axialen Richtung zugewandt ist, dazu konfiguriert ist, als Reaktion auf eine Ansammlung des einen oder der mehreren Steuerfluide in einem Bereich zwischen der Busplatte und der Isolierungsplatte, der über mindestens die Blasendichtung fluidisch abgedichtet ist, zuzunehmen.

2. Vorrichtung (500) nach Anspruch 1, wobei:
die ersten Komponenten ferner eine Kathodengasdiffusionsschicht (Kathoden-GDL) umfassen, die benachbart zu dem Kathodenrahmen (1131) liegt und das Kathodenströmungsfeld (1127) bedeckt, wobei die Kathoden-GDL und das Kathodenströmungsfeld dazu konfiguriert sind, eine Strömung von gasförmigem COₓ über die erste Öffnung in einer ersten Richtung quer zu der axialen Richtung und auf verteilte Weise in Bezug auf mindestens eine zweite Richtung quer zu jeder der axialen und der ersten Richtung zu führen; und
die zweiten Komponenten ferner eine poröse Anodentransportschicht (Anoden-PTL) umfassen, die benachbart zu dem Anodenrahmen (1115) liegt und das Anodenströmungsfeld (1111) bedeckt, wobei die Anoden-PTL und das Anodenströmungsfeld (1111) dazu konfiguriert sind, eine Strömung von Anolyt über die zweite Öffnung in einer dritten Richtung quer zu der axialen Richtung und auf verteilte Weise in Bezug auf mindestens die zweite Richtung zu führen.

3. Vorrichtung (500) nach Anspruch 1, wobei der Kathodenrahmen (1131) Folgendes umfasst:
die erste Öffnung, die in einem mittigen Abschnitt des Kathodenrahmens angeordnet ist;
mindestens einen ersten fluidischen Einlassdurchgang (2815, 2817), der fluidisch mit den anodischen Teilen der Zellen verbunden ist;
mindestens einen ersten fluidischen Auslassdurchgang (2819, 2821), der fluidisch mit den anodischen Teilen der Zellen verbunden ist;
mindestens einen zweiten fluidischen Einlassdurchgang (2827), der fluidisch mit der ersten Öffnung verbunden ist; und
mindestens einen zweiten fluidischen Auslassdurchgang (2829), der fluidisch mit der ersten Öffnung verbunden ist.

4. Vorrichtung (500) nach Anspruch 3, wobei:
der Kathodenrahmen (1131) eine der MEA zugewandte erste Fläche und eine von der ersten Fläche abgewandte zweite Fläche umfasst; und
die zweite Fläche des Kathodenrahmens (1131) Folgendes umfasst:
mindestens einen ersten Vorsprung, durch den sich der mindestens eine erste fluidische Einlassdurchgang (2815, 2817) erstreckt;
mindestens einen zweiten Vorsprung, durch den sich der mindestens eine erste fluidische Auslassdurchgang (2819, 2821) erstreckt;
mindestens einen dritten Vorsprung, durch den sich der mindestens eine zweite fluidische Einlassdurchgang (2827) erstreckt; und
mindestens einen vierten Vorsprung, durch den sich der mindestens eine zweite fluidische Auslassdurchgang (2829) erstreckt.

5. Vorrichtung (500) nach Anspruch 4, wobei:
der mindestens eine erste Vorsprung des Kathodenrahmens (1131) dazu angeordnet und konfiguriert ist, sich derart durch das mindestens eine erste Loch in einer ersten Separatorplatte aus den Separatorplatten (1107) zu erstrecken und an dem Anodenrahmen (1115) einer ersten benachbarten Zelle aus den Zellen (501) anzuliegen, dass der mindestens eine erste fluidische Einlassdurchgang (2815, 2817) des Kathodenrahmens im Wesentlichen in der axialen Richtung mit dem mindestens einen dritten fluidischen Einlassdurchgang des Anodenrahmens der ersten benachbarten Zelle fluchtet;
der mindestens eine zweite Vorsprung des Kathodenrahmens (1131) dazu angeordnet und konfiguriert ist, sich derart durch das mindestens eine zweite Loch in der ersten Separatorplatte zu erstrecken und an dem Anodenrahmen (1115) der ersten benachbarten Zelle anzuliegen, dass der mindestens eine erste fluidische Auslassdurchgang des Kathodenrahmens im Wesentlichen in der axialen Richtung mit dem mindestens einen dritten fluidischen Auslassdurchgang des Anodenrahmens der ersten benachbarten Zelle fluchtet;
der mindestens eine dritte Vorsprung des Kathodenrahmens (1131) dazu angeordnet und konfiguriert ist, sich derart durch das mindestens eine dritte Loch in der ersten Separatorplatte zu erstrecken und an dem Anodenrahmen (1115) der ersten benachbarten Zelle anzuliegen, dass der mindestens eine zweite fluidische Einlassdurchgang des Kathodenrahmens im Wesentlichen in der axialen Richtung mit dem mindestens einen vierten fluidischen Einlassdurchgang des Anodenrahmens der ersten benachbarten Zelle fluchtet; und
der mindestens eine vierte Vorsprung des Kathodenrahmens (1131) dazu angeordnet und konfiguriert ist, sich derart durch das mindestens eine vierte Loch in der ersten Separatorplatte zu erstrecken und an dem Anodenrahmen (1115) der ersten benachbarten Zelle anzuliegen, dass der mindestens eine zweite fluidische Auslassdurchgang des Kathodenrahmens im Wesentlichen in der axialen Richtung mit dem mindestens einen vierten fluidischen Auslassdurchgang des Anodenrahmens (1115) der ersten benachbarten Zelle fluchtet.

6. Vorrichtung (500) nach Anspruch 1, wobei:
der Kathodenrahmen (1131) ferner eine Vielzahl von ersten Kathodenbefestigungsmitteldurchlässen (2837) umfasst, die um einen Randbereich des Kathodenrahmens angeordnet sind, wobei der Randbereich die erste Öffnung des Kathodenrahmens umschließt; und
der Anodenrahmen (1115) ferner Folgendes umfasst:
eine Vielzahl von ersten Anodenbefestigungsmitteldurchlässen (3761), die um einen Randbereich des Anodenrahmens angeordnet sind, wobei der Randbereich die zweite Öffnung des Anodenrahmens umschließt, wobei die ersten Kathodenbefestigungsmitteldurchlässe in der axialen Richtung im Wesentlichen mit den ersten Anodenbefestigungsmitteldurchlässen fluchten; und
eine Vielzahl von ersten Einnietmuttern (1135), wobei jede erste Einnietmutter aus den ersten Einnietmuttern in einem oder dem anderen eines entsprechenden der ersten Anodenbefestigungsmitteldurchlässe und eines entsprechenden der ersten Kathodenbefestigungsmitteldurchlässe vorgesehen ist, wobei die ersten Einnietmuttern dazu konfiguriert sind, eine Grenzfläche mit entsprechenden Rahmenbefestigungsmitteln aus den Rahmenbefestigungsmitteln aufzuweisen.

7. Vorrichtung (500) nach Anspruch 2, wobei:
die ersten Komponenten ferner Folgendes umfassen:
einen ersten Stützrahmen (1123), der zwischen die Kathoden-GDL und den Kathodenrahmen (1131) zwischengeschaltet ist, wobei der erste Stützrahmen eine erste Rahmenöffnung umfasst, die einen Abschnitt der Kathoden-GDL gegenüber dem Kathodenströmungsfeld freilegt, wobei der Abschnitt der Kathoden-GDL an dem Kathodenströmungsfeld anliegt; und
einen zweiten Stützrahmen (1125), der zwischen die MEA und die Anoden-PTL zwischengeschaltet ist, wobei der zweite Stützrahmen eine zweite Rahmenöffnung umfasst, die einen Abschnitt der MEA gegenüber der Anoden-PTL freilegt, wobei der Abschnitt der MEA an der Anoden-PTL anliegt; und
der erste Stützrahmen, die Kathoden-GDL, die MEA und der zweite Stützrahmen eine modularisierte MEA-Baugruppe (301, 401) bilden.

8. Vorrichtung (500) nach Anspruch 7, wobei:
die ersten Komponenten ferner Folgendes umfassen:
eine erste Kathodendichtung (1129), die zwischen den ersten Stützrahmen und den Kathodenrahmen (1131) zwischengeschaltet ist, wobei die erste Kathodendichtung die erste Öffnung in dem Kathodenrahmen umschließt, um eine erste fluidische Abdichtung um das Kathodenströmungsfeld herum zu bilden; und
eine zweite Kathodendichtung (1133), die zwischen eine erste Separatorplatte aus den Separatorplatten und den Kathodenrahmen zwischengeschaltet ist, wobei die zweite Kathodendichtung die erste Öffnung in dem Kathodenrahmen (1131) umschließt, um eine zweite fluidische Abdichtung um das Kathodenströmungsfeld herum zu bilden;
die zweiten Komponenten ferner Folgendes umfassen:
einen ersten Anodendichtungssatz (1113); und
einen zweiten Anodendichtungssatz (1117);
der erste Anodendichtungssatz (1113) Folgendes umfasst:
eine erste Anodendichtung, die zwischen den zweiten Stützrahmen und den Anodenrahmen (1115) zwischengeschaltet ist, wobei die erste Anodendichtung die zweite Öffnung in dem Anodenrahmen umschließt, um eine erste fluidische Abdichtung um das Anodenströmungsfeld herum zu bilden;
mindestens eine zweite Anodendichtung, die zwischen den Kathodenrahmen (1131) und den Anodenrahmen (1115) zwischengeschaltet ist, wobei die mindestens eine zweite Anodendichtung den mindestens einen ersten fluidischen Einlassdurchgang des Kathodenrahmens und den mindestens einen dritten fluidischen Einlassdurchgang der Anode umschließt, um mindestens eine fluidische Abdichtung zu bilden;
mindestens eine dritte Anodendichtung, die zwischen den Kathodenrahmen (1131) und den Anodenrahmen (1115) zwischengeschaltet ist, wobei die mindestens eine dritte Anodendichtung den mindestens einen ersten fluidischen Auslassdurchgang in dem Kathodenrahmen und den mindestens einen dritten fluidischen Auslassdurchgang in dem Anodenrahmen umschließt, um mindestens eine fluidische Abdichtung zu bilden;
mindestens eine vierte Anodendichtung, die zwischen den Kathodenrahmen (1131) und den Anodenrahmen (1115) zwischengeschaltet ist, wobei die mindestens eine dritte Anodendichtung den mindestens einen zweiten fluidischen Einlassdurchgang in dem Kathodenrahmen und den mindestens einen vierten fluidischen Einlassdurchgang in dem Anodenrahmen umschließt, um mindestens eine fluidische Abdichtung zu bilden; und
mindestens eine fünfte Anodendichtung, die zwischen den Kathodenrahmen (1131) und den Anodenrahmen (1115) zwischengeschaltet ist, wobei die mindestens eine fünfte Anodendichtung den mindestens einen zweiten fluidischen Auslassdurchgang und den mindestens einen vierten fluidischen Auslassdurchgang in dem Anodenrahmen umschließt, um mindestens eine fluidische Abdichtung zu bilden; und
der zweite Anodendichtungssatz (1117) Folgendes umfasst:
eine sechste Anodendichtung, die zwischen den Anodenrahmen und eine zweite Separatorplatte aus den Separatorplatten zwischengeschaltet ist, wobei die sechste Anodendichtung die zweite Öffnung in dem Anodenrahmen umschließt, um eine zweite fluidische Abdichtung um das Anodenströmungsfeld (1111) herum zu bilden;
mindestens eine siebte Anodendichtung, die zwischen den Anodenrahmen und die zweite Separatorplatte zwischengeschaltet ist, wobei die mindestens eine siebte Anodendichtung das mindestens eine erste Loch in der zweiten Separatorplatte und den mindestens einen dritten fluidischen Einlassdurchgang in dem Anodenrahmen umschließt, um mindestens eine fluidische Abdichtung zu bilden;
mindestens eine achte Anodendichtung, die zwischen den Anodenrahmen und die zweite Separatorplatte zwischengeschaltet ist, wobei die mindestens eine achte Anodendichtung das mindestens eine zweite Loch in der zweiten Separatorplatte und den mindestens einen dritten fluidischen Auslassdurchgang in dem Anodenrahmen umschließt, um mindestens eine fluidische Abdichtung zu bilden;
mindestens eine neunte Anodendichtung, die zwischen den Anodenrahmen und die zweite Separatorplatte zwischengeschaltet ist, wobei die mindestens eine neunte Anodendichtung das mindestens eine dritte Loch in der zweiten Separatorplatte und den mindestens einen vierten fluidischen Einlassdurchgang in dem Anodenrahmen umschließt, um mindestens eine fluidische Abdichtung zu bilden; und
mindestens eine zehnte Anodendichtung, die zwischen den Anodenrahmen und die zweite Separatorplatte zwischengeschaltet ist, wobei die mindestens eine neunte Anodendichtung das mindestens eine vierte Loch in der zweiten Separatorplatte und den mindestens einen vierten fluidischen Auslassdurchgang in dem Anodenrahmen umschließt, um mindestens eine fluidische Abdichtung zu bilden.

9. Vorrichtung (500) nach Anspruch 1, wobei:
jede der Separatorplatten (1107) Folgendes umfasst:
eine Vielzahl von Befestigungsmitteldurchlässen, durch die sich die Rahmenbefestigungsmittel jeweils erstrecken;
mindestens ein erstes Loch, durch das sich ein Einlassströmungsweg von Anolyt erstreckt;
mindestens ein zweites Loch, durch das sich ein Auslassströmungsweg von Anolyt erstreckt;
mindestens ein drittes Loch, durch das sich ein Einlassströmungsweg von gasförmigem COₓ erstreckt; und
mindestens ein viertes Loch, durch das sich ein Auslassströmungsweg von COₓ-Reduktionsnebenprodukt erstreckt;
die erste Endbaugruppe ferner eine erste Isolierungsplatte, einen Verteiler und eine erste Busplatte zwischen der ersten Endplatte und der Kathodengrenzflächenbaugruppe umfasst;
der Verteiler Folgendes umfasst:
mindestens einen ersten Einlass, der über den Einlassströmungsweg von Anolyt fluidisch mit den anodischen Teilen der Zellen verbunden ist;
mindestens einen ersten Auslass, der über den Auslassströmungsweg von Anolyt fluidisch mit den anodischen Teilen der Zellen verbunden ist;
mindestens einen zweiten Einlass, der über den Einlassströmungsweg von gasförmigem COₓ fluidisch mit den kathodischen Teilen der Zellen verbunden ist; und
mindestens einen zweiten Auslass, der über den Auslassströmungsweg von COₓ-Reduktionsnebenprodukt fluidisch mit den kathodischen Teilen der Zellen verbunden ist;
die erste Busplatte dazu konfiguriert ist, ein erstes elektrisches Potential aufzunehmen;
die erste Isolierungsplatte dazu konfiguriert ist, die erste Endplatte elektrisch von der ersten Busplatte zu isolieren, wobei sich der Einlassströmungsweg von Anolyt, der Auslassströmungsweg von Anolyt, der Einlassströmungsweg von gasförmigem COₓ und der Auslassströmungsweg von COₓ-Reduktionsnebenprodukt nicht in die Busplatte und die erste Isolierungsplatte erstrecken.

10. Vorrichtung (500) nach Anspruch 1, wobei:
die zweite Endbaugruppe ferner eine zweite Busplatte und eine zweite Isolierungsplatte umfasst, die nacheinander in der axialen Richtung zwischen der Anodengrenzflächenbaugruppe 509 und der zweiten Endplatte gestapelt sind;
die zweite Busplatte dazu konfiguriert ist, ein zweites elektrisches Potential aufzunehmen; und
die zweite Isolierungsplatte dazu konfiguriert ist, die zweite Endplatte elektrisch von der zweiten Busplatte zu isolieren.

11. Vorrichtung (500) nach Anspruch 10, wobei:
die zweite Endplatte Folgendes umfasst:
einen ersten Hauptkörper;
einen Vorsprung der zweiten Endplatte, der sich von dem ersten Hauptkörper in der axialen Richtung erstreckt; und
eine Öffnung der zweiten Endplatte, die sich in einen mittigen Abschnitt des Vorsprungs der zweiten Endplatte in einer zu der axialen Richtung entgegengesetzten Richtung erstreckt und an einer den Zellen zugewandten vertieften Fläche endet;
die zweite Endbaugruppe ferner einen Kolben 10105 umfasst, der zwischen die zweite Isolierungsplatte und die zweite Endplatte zwischengeschaltet ist, wobei der Kolben Folgendes umfasst:
einen zweiten Hauptkörper; und
einen Kolbenvorsprung, der sich von dem zweiten Hauptkörper in der zu der axialen Richtung entgegengesetzten Richtung erstreckt und an einer der vertieften Fläche zugewandten vorspringenden Fläche endet;
mindestens ein Abschnitt des Kolbenvorsprungs verschiebbar in mindestens einem Abschnitt der Öffnung der zweiten Endplatte vorgesehen ist;
die zweite Endplatte ferner einen oder mehrere Durchlässe umfasst, die fluidisch mit der Öffnung der zweiten Endplatte verbunden sind, wobei der eine oder die mehreren Durchlässe dazu konfiguriert sind, ein oder mehrere Steuerfluide aufzunehmen;
der Kolbenvorsprung eine Vielzahl von Kolbendichtungen 10119 umfasst, die den Kolbenvorsprung umschließen und in der axialen Richtung voneinander versetzt sind, wobei die Kolbendichtungen derart eine Grenzfläche mit einer oder mehreren inneren Seitenwänden der Öffnung der zweiten Endplatte aufweisen, dass die Öffnung der zweiten Endplatte, der Kolbenvorsprung und die Kolbendichtungen 10119 einen Hohlraum innerhalb der zweiten Endbaugruppe bilden; und
ein Abstand in der axialen Richtung zwischen der vorspringenden Fläche und der vertieften Fläche dazu konfiguriert ist, als Reaktion auf eine Ansammlung des einen oder der mehreren Steuerfluide in dem Hohlraum zuzunehmen.

12. Vorrichtung (500) nach Anspruch 11, wobei:
die zweite Endbaugruppe ferner ein Vielzahl von Vorspannelementen (10117) umfasst;
der Kolbenvorsprung eine Vielzahl von Kolbenvorsprungsöffnungen umfasst, die sich in der axialen Richtung in die vorspringende Fläche erstrecken;
die zweite Endplatte ferner eine Vielzahl von Stützvorsprüngen umfasst, die sich in der axialen Richtung von der vertieften Fläche erstrecken und in Übereinstimmung mit den Kolbenvorsprungsöffnungen angeordnet sind;
die Vorspannelemente (10117) jeweils derart über entsprechende Stützvorsprünge aus den Stützvorsprüngen in der Öffnung der zweiten Endplatte gestützt sind, dass in einem ersten komprimierten Zustand der zweiten Endbaugruppe die Vorspannelemente zwischen der vorspringenden Fläche und der vertieften Fläche komprimiert sind und sich jeweilige Abschnitte der Stützvorsprünge mindestens teilweise in entsprechende Kolbenvorsprungsöffnungen aus den Kolbenvorsprungsöffnungen erstrecken;
die zweite Endplatte ferner einen oder mehrere Durchlässe umfasst, die fluidisch mit der Öffnung der zweiten Endplatte verbunden sind, wobei der eine oder die mehreren Durchlässe dazu konfiguriert sind, ein oder mehrere Steuerfluide aufzunehmen;
der Kolbenvorsprung eine Vielzahl von Kolbendichtungen (10119) umfasst, die den Kolbenvorsprung umschließen und in der axialen Richtung voneinander versetzt sind, wobei die Kolbendichtungen derart eine Grenzfläche mit einer oder mehreren inneren Seitenwänden der Öffnung der zweiten Endplatte aufweisen, dass die Öffnung der zweiten Endplatte, der Kolbenvorsprung und die Kolbendichtungen einen Hohlraum innerhalb der zweiten Endbaugruppe bilden; und
ein Abstand in der axialen Richtung zwischen der vorspringenden Fläche und der vertieften Fläche dazu konfiguriert ist, als Reaktion auf eine Ansammlung des einen oder der mehreren Steuerfluide in dem Hohlraum zuzunehmen.

## Revendications

1. Appareil d'électrolyse de COₓ (500) comprenant :
un premier ensemble d'extrémité comprenant une première plaque d'extrémité (519) et un ensemble d'interface de cathode (505) ; un second ensemble d'extrémité comprenant une seconde plaque d'extrémité (525), un ensemble d'interface d'anode (509), et un joint à vessie (559), dans lequel le second ensemble d'extrémité est couplé au premier ensemble d'extrémité via une pluralité d'éléments de mise en tension (527) ;
une pluralité de plaques séparatrices (1107) ; et
une pluralité de cellules d'électrolyse de COₓ (501) qui sont chacune formées d'une pluralité d'unités de répétition (503, 1100), dans lequel la pluralité de cellules sont interposées entre les premier et second ensembles d'extrémité et agencées en un empilement le long d'une direction axiale, chaque cellule parmi les cellules (501) comprenant un exemplaire de premiers composants et un exemplaire de seconds composants,
dans lequel les premiers composants comprennent :
un ensemble électrode-membrane (EEM ; 301, 401) ayant une partie cathodique (303, 403), une partie anodique (305, 405), et un séparateur entre la partie cathodique et la partie anodique ;
un cadre de cathode (1131) adjacent à la partie cathodique ; et
un champ d'écoulement de cathode (1127) au moins partiellement disposé dans une première ouverture dans le cadre de cathode,
dans lequel les seconds composants comprennent :
un cadre d'anode (1115) adjacent à la partie anodique de l'EEM ; et
un champ d'écoulement d'anode (1111) au moins partiellement disposé dans une seconde ouverture dans le cadre d'anode,
dans lequel chaque unité de répétition (503, 1100) parmi les unités de répétition comprend :
un exemplaire des premiers composants ;
un exemplaire des seconds composants ; et
la plaque séparatrice (1107) qui est interposée entre le cadre de cathode (1131) de cet exemplaire des premiers composants et le cadre d'anode (1115) de cet exemplaire des seconds composants, la plaque séparatrice (1107) étant interposée entre cet exemplaire des premiers composants et cet exemplaire des seconds composants ;
dans lequel l'ensemble d'interface de cathode (505) comprend :
un exemplaire des premiers composants ; et
une plaque séparatrice d'interface de cathode (1701) interposée entre la première plaque d'extrémité et une première unité de répétition parmi les unités de répétition (503, 1100) ;
dans lequel l'ensemble d'interface d'anode (509) comprend :
un exemplaire des seconds composants ;
et une plaque séparatrice d'interface d'anode (4703) interposée entre une seconde unité de répétition parmi les unités de répétition et la seconde plaque d'extrémité ;
dans lequel les cadres de cathode (1131) et d'anode (1115) de cellules adjacentes parmi les cellules sont couplés les uns aux autres via une pluralité correspondante d'éléments de fixation de cadre avec une plaque séparatrice parmi les plaques séparatrices (1107) interposée entre eux, les éléments de fixation de cadre étant différents des éléments de mise en tension (527) ;
une première cellule d'extrémité est formée entre l'ensemble d'interface de cathode (505) et l'exemplaire des seconds composants de la première unité de répétition, la première cellule d'extrémité étant interposée entre la première plaque d'extrémité et la pluralité de cellules (501) ;
une seconde cellule d'extrémité est formée entre l'exemplaire des premiers composants de la seconde unité de répétition et l'ensemble d'interface d'anode (509), la seconde cellule d'extrémité étant interposée entre la pluralité de cellules (501) et la seconde plaque d'extrémité ;
une plaque d'isolation (523) comprenant :
un premier évidement formé dans une partie centrale de la plaque d'isolation ;
un second évidement encerclant une région centrale de la partie centrale, le second évidement supportant le joint à vessie (559) en son sein ; et
un orifice (8631) configuré pour recevoir un ou plusieurs fluides de commande ;
une plaque de barre omnibus (521) disposée de manière coulissante dans le premier évidement et configurée pour venir en butée contre le joint à vessie (559) et/ou une surface du premier évidement faisant face à la plaque de barre omnibus (521) dans la direction axiale ; et
une distance dans la direction axiale entre la plaque de barre omnibus et la surface du premier évidement faisant face à la plaque de barre omnibus dans la direction axiale est configurée pour augmenter en réponse à l'accumulation des un ou plusieurs fluides de commande dans une zone entre la plaque de barre omnibus et la plaque d'isolation qui est étanchéifiée de manière fluidique via au moins le joint à vessie.

2. Appareil (500) selon la revendication 1, dans lequel :
les premiers composants comprennent en outre une couche de diffusion de gaz (CDG) de cathode adjacente au cadre de cathode (1131) et recouvrant le champ d'écoulement de cathode (1127), la CDG de cathode et le champ d'écoulement de cathode étant configurés pour guider un écoulement de COₓ gazeux à travers la première ouverture dans une première direction transversale à la direction axiale et d'une manière distribuée par rapport à au moins une deuxième direction transversale à chacune des directions axiale et première ; et
les seconds composants comprennent en outre une couche de transport poreuse (CTP) d'anode adjacente au cadre d'anode (1115) et recouvrant le champ d'écoulement d'anode (1111), la CTP d'anode et le champ d'écoulement d'anode (1111) étant configurés pour guider un écoulement d'anolyte à travers la seconde ouverture dans une troisième direction transversale à la direction axiale et d'une manière distribuée par rapport à au moins la deuxième direction.

3. Appareil (500) selon la revendication 1, dans lequel le cadre de cathode (1131) comprend :
la première ouverture agencée dans une partie centrale du cadre de cathode ;
au moins un premier passage d'entrée fluidique (2815, 2817) connecté de manière fluidique aux parties anodiques des cellules ;
au moins un premier passage de sortie fluidique (2819, 2821) connecté de manière fluidique aux parties anodiques des cellules ;
au moins un second passage d'entrée fluidique (2827) connecté de manière fluidique à la première ouverture ; et
au moins un second passage de sortie fluidique (2829) connecté de manière fluidique à la première ouverture.

4. Appareil (500) selon la revendication 3, dans lequel :
le cadre de cathode (1131) comprend une première surface faisant face à l'EEM et une seconde surface faisant face à l'opposé de la première surface ; et
la seconde surface du cadre de cathode (1131) comprend :
au moins une première saillie à travers laquelle l'au moins un premier passage d'entrée fluidique (2815, 2817) s'étend ;
au moins une deuxième saillie à travers laquelle l'au moins un premier passage de sortie fluidique (2819, 2821) s'étend ;
au moins une troisième saillie à travers laquelle l'au moins un second passage d'entrée fluidique (2827) s'étend ; et
au moins une quatrième saillie à travers laquelle l'au moins un second passage de sortie fluidique (2829) s'étend.

5. Appareil (500) selon la revendication 4, dans lequel :
l'au moins une première saillie du cadre de cathode (1131) est agencée et configurée pour s'étendre à travers l'au moins un premier trou dans une première plaque séparatrice parmi les plaques séparatrices (1107) et venir en butée contre le cadre d'anode (1115) d'une première cellule adjacente parmi les cellules (501) de sorte que l'au moins un premier passage d'entrée fluidique (2815, 2817) du cadre de cathode soit substantiellement aligné dans la direction axiale avec l'au moins un troisième passage d'entrée fluidique du cadre d'anode de la première cellule adjacente ;
l'au moins une deuxième saillie du cadre de cathode (1131) est agencée et configurée pour s'étendre à travers l'au moins un deuxième trou dans la première plaque séparatrice et venir en butée contre le cadre d'anode (1115) d'une première cellule adjacente de sorte que l'au moins un premier passage de sortie fluidique du cadre de cathode soit substantiellement aligné dans la direction axiale avec l'au moins un troisième passage de sortie fluidique du cadre d'anode de la première cellule adjacente ;
l'au moins une troisième saillie du cadre de cathode (1131) est agencée et configurée pour s'étendre à travers l'au moins un troisième trou dans la première plaque séparatrice et venir en butée contre le cadre d'anode (1115) d'une première cellule adjacente de sorte que l'au moins un deuxième passage d'entrée fluidique du cadre de cathode soit substantiellement aligné dans la direction axiale avec l'au moins un quatrième passage d'entrée fluidique du cadre d'anode de la première cellule adjacente ; et
l'au moins une quatrième saillie du cadre de cathode (1131) est agencée et configurée pour s'étendre à travers l'au moins un quatrième trou dans la première plaque séparatrice et venir en butée contre le cadre d'anode (1115) d'une première cellule adjacente de sorte que l'au moins un deuxième passage de sortie fluidique du cadre de cathode soit substantiellement aligné dans la direction axiale avec l'au moins un quatrième passage de sortie fluidique du cadre d'anode (1115) de la première cellule adjacente.

6. Appareil (500) selon la revendication 1, dans lequel :
le cadre de cathode (1131) comprend en outre une pluralité de premiers orifices d'élément de fixation de cathode (2837) agencés autour d'une zone périphérique du cadre de cathode, la zone périphérique encerclant la première ouverture du cadre de cathode ; et
le cadre d'anode (1115) comprend en outre :
une pluralité de premiers orifices d'élément de fixation d'anode (3761) agencés autour d'une zone périphérique du cadre d'anode, la zone périphérique encerclant la seconde ouverture du cadre d'anode, les premiers orifices d'élément de fixation de cathode étant substantiellement alignés avec les premiers orifices d'élément de fixation d'anode dans la direction axiale ; et
une pluralité de premiers écrous auto-sertissables (1135), chaque premier écrou auto-sertissable parmi les premiers écrous auto-sertissables étant disposé dans l'un ou l'autre d'un orifice correspondant parmi les premiers orifices d'élément de fixation d'anode et d'un orifice correspondant parmi les premiers orifices d'élément de fixation de cathode, les premiers écrous auto-sertissables étant configurés pour s'interfacer avec des éléments de fixation de cadre correspondants parmi les éléments de fixation de cadre.

7. Appareil (500) selon la revendication 2, dans lequel :
les premiers composants comprennent en outre :
un premier cadre de support (1123) interposé entre la CDG de cathode et le cadre de cathode (1131), le premier cadre de support comprenant une première ouverture de cadre exposant une partie de la CDG de cathode au champ d'écoulement de cathode, la partie de la CDG de cathode venant en butée contre le champ d'écoulement de cathode ; et
un second cadre de support (1125) interposé entre l'EEM et la CTP d'anode, le second cadre de support comprenant une seconde ouverture de cadre exposant une partie de l'EEM à la CTP d'anode, la partie de l'EEM venant en butée contre la CTP d'anode ; et
le premier cadre de support, la CDG de cathode, l'EEM, et le second cadre de support forment un ensemble EEM monobloc (301, 401).

8. Appareil (500) selon la revendication 7, dans lequel :
les premiers composants comprennent en outre :
un premier joint de cathode (1129) interposé entre le premier cadre de support et le cadre de cathode (1131), le premier joint de cathode encerclant la première ouverture dans le cadre de cathode pour former un premier joint d'étanchéité fluidique autour du champ d'écoulement de cathode ; et
un second joint de cathode (1133) interposé entre une première plaque séparatrice parmi les plaques séparatrices et le cadre de cathode, le second joint de cathode encerclant la première ouverture dans le cadre de cathode (1131) pour former un second joint d'étanchéité fluidique autour du champ d'écoulement de cathode ;
les seconds composants comprennent en outre :
un premier ensemble de joints d'anode (1113) ; et
un second ensemble de joints d'anode (1117) ;
le premier ensemble de joints d'anode (1113) comprend :
un premier joint d'anode interposé entre le second cadre de support et le cadre d'anode (1115), le premier joint d'anode encerclant la seconde ouverture dans le cadre d'anode pour former un premier joint d'étanchéité fluidique autour du champ d'écoulement d'anode ;
au moins un deuxième joint d'anode interposé entre le cadre de cathode (1131) et le cadre d'anode (1115), l'au moins un deuxième joint d'anode encerclant l'au moins un premier passage d'entrée fluidique du cadre de cathode et l'au moins un troisième passage d'entrée fluidique de l'anode pour former au moins un joint d'étanchéité fluidique ;
au moins un troisième joint d'anode interposé entre le cadre de cathode (1131) et le cadre d'anode (1115), l'au moins un troisième joint d'anode encerclant l'au moins un premier passage de sortie fluidique dans le cadre de cathode et l'au moins un troisième passage de sortie fluidique dans le cadre d'anode pour former au moins un joint d'étanchéité fluidique ;
au moins un quatrième joint d'anode interposé entre le cadre de cathode (1131) and le cadre d'anode (1115), l'au moins un troisième joint d'anode encerclant l'au moins un second passage d'entrée fluidique dans le cadre de cathode et l'au moins un quatrième passage d'entrée fluidique dans le cadre d'anode pour former au moins un joint d'étanchéité fluidique ; et
au moins un cinquième joint d'anode interposé entre le cadre de cathode (1131) et le cadre d'anode (1115), l'au moins un cinquième joint d'anode encerclant l'au moins un second passage de sortie fluidique et l'au moins un quatrième passage de sortie fluidique dans le cadre d'anode pour former au moins un joint d'étanchéité fluidique ; et
le second ensemble de joints d'anode (1117) comprend :
un sixième joint d'anode interposé entre le cadre d'anode et une seconde plaque séparatrice parmi les plaques séparatrices, le sixième joint d'anode encerclant la seconde ouverture dans le cadre d'anode pour former un second joint d'étanchéité fluidique autour du champ d'écoulement d'anode (1111) ;
au moins un septième joint d'anode interposé entre le cadre d'anode et la seconde plaque séparatrice, l'au moins un septième joint d'anode encerclant l'au moins un premier trou dans la seconde plaque séparatrice et l'au moins un troisième passage d'entrée fluidique dans le cadre d'anode pour former au moins un joint d'étanchéité fluidique ;
au moins un huitième joint d'anode interposé entre le cadre d'anode et la seconde plaque séparatrice, l'au moins un huitième joint d'anode encerclant l'au moins un deuxième trou dans la seconde plaque séparatrice et l'au moins un troisième passage de sortie fluidique dans le cadre d'anode pour former au moins un joint d'étanchéité fluidique ;
au moins un neuvième joint d'anode interposé entre le cadre d'anode et la seconde plaque séparatrice, l'au moins un neuvième joint d'anode encerclant l'au moins un troisième trou dans la seconde plaque séparatrice et l'au moins un quatrième passage d'entrée fluidique dans le cadre d'anode pour former au moins un joint d'étanchéité fluidique ; et
au moins un dixième joint d'anode interposé entre le cadre d'anode et la seconde plaque séparatrice, l'au moins un neuvième joint d'anode encerclant l'au moins un quatrième trou dans la seconde plaque séparatrice et l'au moins un quatrième passage de sortie fluidique dans le cadre d'anode pour former au moins un joint d'étanchéité fluidique.

9. Appareil (500) selon la revendication 1, dans lequel :
chacune des plaques séparatrices (1107) comprend :
une pluralité d'orifices d'élément de fixation à travers lesquels les éléments de fixation de cadre s'étendent respectivement ;
au moins un premier trou à travers lequel un trajet d'écoulement d'anolyte d'entrée s'étend ;
au moins un deuxième trou à travers lequel un trajet d'écoulement d'anolyte de sortie s'étend ;
au moins un troisième trou à travers lequel un trajet d'écoulement de COₓ gazeux d'entrée s'étend ; et
au moins un quatrième trou à travers lequel un trajet d'écoulement de sous-produit de réduction de COₓ de sortie s'étend ;
le premier ensemble d'extrémité comprend en outre une première plaque d'isolation, un collecteur, et une première plaque de barre omnibus entre la première plaque d'extrémité et l'ensemble d'interface de cathode ;
le collecteur comprend :
au moins une première entrée connectée de manière fluidique aux parties anodiques des cellules via le trajet d'écoulement d'anolyte d'entrée ;
au moins une première sortie connectée de manière fluidique aux parties anodiques des cellules via le trajet d'écoulement d'anolyte de sortie ;
au moins une deuxième entrée connectée de manière fluidique aux parties cathodiques des cellules via le trajet d'écoulement de COₓ gazeux d'entrée ; et
au moins une deuxième sortie connectée de manière fluidique aux parties cathodiques des cellules via le trajet d'écoulement de sous-produit de réduction de COₓ de sortie ;
la première plaque de barre omnibus est configurée pour recevoir un premier potentiel électrique ;
la première plaque d'isolation est configurée pour isoler électriquement la première plaque d'extrémité de la première plaque de barre omnibus, dans lequel le trajet d'écoulement d'anolyte d'entrée, le trajet d'écoulement d'anolyte de sortie, le trajet d'écoulement de COₓ gazeux d'entrée, et le trajet d'écoulement de sous-produit de réduction de COₓ de sortie ne s'étendent pas dans la plaque de barre omnibus et la première plaque d'isolation.

10. Appareil (500) selon la revendication 1, dans lequel :
le second ensemble d'extrémité comprend en outre une seconde plaque de barre omnibus et une seconde plaque d'isolation empilées séquentiellement dans la direction axiale entre l'ensemble d'interface d'anode (509) et la seconde plaque d'extrémité ;
la seconde plaque de barre omnibus est configurée pour recevoir un second potentiel électrique ; et
la seconde plaque d'isolation est configurée pour isoler électriquement la seconde plaque d'extrémité de la seconde plaque de barre omnibus.

11. Appareil (500) selon la revendication 10, dans lequel :
la seconde plaque d'extrémité comprend :
un premier corps principal ;
une saillie de seconde plaque d'extrémité s'étendant à partir du premier corps principal dans la direction axiale ; et
une ouverture de seconde plaque d'extrémité s'étendant dans une partie centrale de la saillie de seconde plaque d'extrémité dans une direction opposée à la direction axiale et se terminant au niveau d'une surface évidée faisant face aux cellules ;
le second ensemble d'extrémité comprend en outre un piston (10105) interposé entre la seconde plaque d'isolation et la seconde plaque d'extrémité, le piston comprenant :
un second corps principal ; et
une saillie de piston s'étendant à partir du second corps principal dans la direction opposée à la direction axiale et se terminant au niveau d'une surface saillante faisant face à la surface évidée ;
au moins une partie de la saillie de piston est disposée de manière coulissante dans au moins une partie de l'ouverture de seconde plaque d'extrémité ;
la seconde plaque d'extrémité comprend en outre un ou plusieurs orifices connectés de manière fluidique à l'ouverture de seconde plaque d'extrémité, les un ou plusieurs orifices étant configurés pour recevoir un ou plusieurs fluides de commande ; la saillie de piston comprend une pluralité de joints de piston (10119) encerclant la saillie de piston et décalés les uns des autres dans la direction axiale, les joints de piston s'interfaçant avec une ou plusieurs parois latérales internes de l'ouverture de seconde plaque d'extrémité de sorte que l'ouverture de seconde plaque d'extrémité, la saillie de piston, et les joints de piston (10119) forment une cavité à l'intérieur du second ensemble d'extrémité ; et
une distance dans la direction axiale entre la surface saillante et la surface évidée est configurée pour augmenter en réponse à l'accumulation des un ou plusieurs fluides de commande dans la cavité.

12. Appareil (500) selon la revendication 11, dans lequel :
le second ensemble d'extrémité comprend en outre une pluralité d'éléments de sollicitation (10117) ;
la saillie de piston comprend une pluralité d'ouvertures de saillie de piston s'étendant dans la surface saillante dans la direction axiale ;
la seconde plaque d'extrémité comprend en outre une pluralité de saillies de support s'étendant dans la direction axiale à partir de la surface évidée et agencées en correspondance avec les ouvertures de saillie de piston ;
les éléments de sollicitation (10117) sont respectivement supportés dans l'ouverture de seconde plaque d'extrémité via des saillies de support correspondantes parmi les saillies de support de sorte que, dans un premier état comprimé du second ensemble d'extrémité, les éléments de sollicitation soient comprimés entre la surface saillante et la surface évidée et que des parties respectives des saillies de support s'étendent au moins partiellement dans des ouvertures de saillie de piston correspondantes parmi les ouvertures de saillie de piston ;
la seconde plaque d'extrémité comprend en outre un ou plusieurs orifices connectés de manière fluidique à l'ouverture de seconde plaque d'extrémité, les un ou plusieurs orifices étant configurés pour recevoir un ou plusieurs fluides de commande ;
la saillie de piston comprend une pluralité de joints de piston (10119) encerclant la saillie de piston et décalés les uns des autres dans la direction axiale, les joints de piston s'interfaçant avec une ou plusieurs parois latérales internes de l'ouverture de seconde plaque d'extrémité de sorte que l'ouverture de seconde plaque d'extrémité, la saillie de piston, et les joints de piston forment une cavité à l'intérieur du second ensemble d'extrémité ; et
une distance dans la direction axiale entre la surface saillante et la surface évidée est configurée pour augmenter en réponse à l'accumulation des un ou plusieurs fluides de commande dans la cavité.
